# EUROPEAN PATENT SPECIFICATION

(11) **EP 0 743 574 B1**
(45) Date of publication and mention of the grant of the patent: **27.12.2000**
(21) Application number: 96303360.0
(22) Date of filing: 14.05.1996
(51) Int. Cl.: G03G 17/10, G03G 17/06

(54) **Migration imaging members**
Bilderzeugungselemente nach dem Migrationsverfahren
Eléments de formation d'images par migration

(30) Priority: 15.05.1995 US 422227
(43) Date of publication of application: 20.11.1996
(73) Proprietor: XEROX CORPORATION, Rochester, New York 14644 (US)
(72) Inventor: Malhotra, Shadi L., Mississauga, Ontario L5L 2A6 (CA); Chen, Liqin, Ontario L5A 3K8 (CA); Perron, Marie-Eve, Montreal, Quebec H4V 2S9 (CA)
(74) Representative: Grünecker, Kinkeldey, Stockmair & Schwanhäusser Anwaltssozietät

(56) References cited:
- WO-A-93/04411
- US-A- 4 101 321
- US-A- 5 240 799

## Description

The present invention is directed to improved migration imaging members. More specifically, the present invention is directed to migration imaging members with improved optical contrast density.

While known apparatus and processes are suitable for their intended purposes, a need remains for improved migration imaging members. In addition, a need remains for migration imaging members with improved optical contrast density. Further, there is a need for migration imaging members wherein the optical density of the Dₘᵢₙ areas of the imaged member is decreased without a corresponding decrease in the optical density of the Dₘₐₓ areas of the imaged member. Additionally, there is a need for migration imaging members wherein the optical density of the Dₘᵢₙ areas of the imaged member with respect to ultraviolet light passing through the imaging member is decreased without a corresponding decrease in the optical density of the Dₘₐₓ areas of the imaged member with respect to ultraviolet light passing through the imaging member.

It is an object of the present invention to provide migration imaging members with the above noted advantages.

These and other objects of the present invention (or specific embodiments thereof) can be achieved by providing a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member wherein the transparentizing agent affects the migration marking material which comes into contact therewith by reducing the optical density of the softenable layer containing the migration marking material. Another embodiment of the present invention is directed to a process which comprises (1) providing a migration imaging member comprising (a) a substrate, (b) a softenable layer comprising a softenable material and a photosensitive migration marking material, and (c) a transparentizing agent which transparentizes migration marking material in contact therewith contained in at least one layer of the migration imaging member; (2) uniformly charging the imaging member; (3) subsequent to step (2), exposing the charged imaging member to activating radiation at a wavelength to which the migration marking material is sensitive; (4) subsequent to step (3), causing the softenable material to soften and enabling a first portion of the migration marking material to migrate through the softenable material toward the substrate in an imagewise pattern while a second portion of the migration marking material remains substantially unmigrated within the softenable layer, wherein subsequent to migration of the first portion of migration marking material, either (a) the first portion of migration marking material contacts the transparentizing agent and the second portion of migration marking material does not contact the transparentizing agent; or (b) the second portion of migration marking material contacts the transparentizing agent and the first portion of migration marking material does not contact the transparentizing agent.

Other embodiments of the invention are defined in the appended claims.

The present invention will be described further, by way of examples, with reference to the accompanying drawings, in which:-
Figure 1 illustrates schematically one migration imaging member suitable for the present invention, wherein a transparentizing agent is included within one or more layers of the imaging member;
Figures 2 and 3 illustrate schematically infrared-sensitive migration imaging members suitable for the present invention, wherein a transparentizing agent is included within one or more layers of the imaging member; and
Figures 4, 5, 6, 7, 8, 9, and 10 illustrate schematically migration imaging members suitable for the present invention, wherein a transparentizing agent is present in a separate transparentizing layer within the imaging member.

The present invention encompasses migration imaging members containing an agent for transparentizing migration marking material in at least one layer of the migration imaging member. The transparentizing agent is a material that affects migration marking material which comes into contact therewith by reducing the optical density of the softenable layer containing the migration marking material in said areas. Thus, in one embodiment of the present invention, when migration marking material migrates selectively through the softenable layer in imagewise fashion, the migrated marking material contacts the transparentizing agent while the unmigrated marking material does not contact the transparentizing agent (or contacts it to a lesser degree than the migrated marking material contacts it), thereby reducing the optical density of the softenable layer in areas wherein the migration marking material has migrated (i.e., in Dₘᵢₙ areas). In another embodiment of the present invention, when migration marking material migrates selectively through the softenable layer in imagewise fashion, the unmigrated marking material contacts the transparentizing agent while the migrated marking material does not contact the transparentizing agent (or contacts it to a lesser degree than the unmigrated marking material contacts it), thereby reducing the optical density of the softenable layer in areas wherein the migration marking material has not migrated.

An example of a migration imaging member suitable for the present invention is illustrated schematically in Figure 1. As illustrated schematically in Figure 1, migration imaging member 1 comprises a substrate 2, an optional adhesive layer 3 situated on the substrate 2, an optional charge blocking layer 4 situated on optional adhesive layer 3, an optional charge transport layer 5 situated on optional charge blocking layer 4, and a softenable layer 6 situated on optional charge transport layer 5, said softenable layer 6 comprising softenable material 7, migration marking material 8 situated at or near the surface of the layer spaced from the substrate, and optional charge transport material 9 dispersed throughout softenable material 7. Optional overcoating layer 10 is situated on the surface of softenable layer 6 spaced from the substrate 2. Any or all of the optional layers and materials can be absent from the imaging member. In addition, any of the optional layers present need not be in the order shown, but can be in any suitable arrangement. The migration imaging member can be in any suitable configuration, such as a web, a foil, a laminate, a strip, a sheet, a coil, a cylinder, a drum, an endless belt, an endless mobius strip, a circular disc, or any other suitable form.

The substrate can be either electrically conductive or electrically insulating. When conductive, the substrate can be opaque, translucent, semitransparent, or transparent, and can be of any suitable conductive material, including copper, brass, nickel, zinc, chromium, stainless steel, conductive plastics and rubbers, aluminum, semitransparent aluminum, steel, cadmium, silver, gold, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. When insulative, the substrate can be opaque, translucent, semitransparent, or transparent, and can be of any suitable insulative material, such as paper, glass, plastic, polyesters such as Mylar® (available from Du Pont) or Melinex® 442 (available from ICI Americas, Inc.), and the like. In addition, the substrate can comprise an insulative layer with a conductive coating, such as vacuum-deposited metallized plastic, such as titanized or aluminized Mylar® polyester, wherein the metallized surface is in contact with the softenable layer or any other layer situated between the substrate and the softenable layer. The substrate has any effective thickness, typically from about 6 to about 250 microns, and preferably from about 50 to about 200 microns, although the thickness can be outside these ranges.

The softenable layer can comprise one or more layers of softenable materials, which can be any suitable material, typically a plastic or thermoplastic material which is soluble in a solvent or softenable, for example, in a solvent liquid, solvent vapor, heat, or any combinations thereof. When the softenable layer is to be softened or dissolved either during or after imaging, it should be soluble in a solvent that does not attack the migration marking material. By softenable is meant any material that can be rendered by a development step as described herein permeable to migration material migrating through its bulk. This permeability typically is achieved by a development step entailing dissolving, melting, or softening by contact with heat, vapors, partial solvents, as well as combinations thereof. Examples of suitable softenable materials include styrene-acrylic copolymers, such as styrene-hexyl methacrylate copolymers, styrene acrylate copolymers, styrene butylmethacrylate copolymers, styrene butylacrylate ethylacrylate copolymers, styrene ethylacrylate acrylic acid copolymers, and the like, polystyrenes, including polyalphamethyl styrene, alkyd substituted polystyrenes, styrene-olefin copolymers, styrene-vinyltoluene copolymers, polyesters, polyurethanes, polycarbonates, polyterpenes, silicone elastomers, mixtures thereof, copolymers thereof, and the like, as well as any other suitable materials as disclosed, for example, in U.S. Patent 3,975,195 and other U.S. patents directed to migration imaging members. The softenable layer can be of any effective thickness, typically from about 1 to about 30 microns, preferably from about 2 to about 25 microns, and more preferably from about 2 to about 10 microns, although the thickness can be outside these ranges. The softenable layer can be applied to the conductive layer by any suitable coating process. Typical coating processes include draw bar coating, spray coating, extrusion, dip coating, gravure roll coating, wire-wound rod coating, air knife coating and the like.

The softenable layer also contains migration marking material. The migration marking material can be electrically photosensitive, photoconductive, or of any other suitable combination of materials, or possess any other desired physical property and still be suitable for use in the migration imaging members of the present invention. The migration marking materials preferably are particulate, wherein the particles are closely spaced from each other. Preferred migration marking materials generally are spherical in shape and submicron in size. The migration marking material generally is capable of substantial photodischarge upon electrostatic charging and exposure to activating radiation and is substantially absorbing and opaque to activating radiation in the spectral region where the photosensitive migration marking particles photogenerate charges. The migration marking material is generally present as a thin layer or monolayer of particles situated at or near the surface of the softenable layer spaced from the conductive layer. When present as particles, the particles of migration marking material preferably have an average diameter of up to 2 microns, and more preferably of from about 0.1 to about 1 micron. The layer of migration marking particles is situated at or near that surface of the softenable layer spaced from or most distant from the conductive layer. Preferably, the particles are situated at a distance of from about 0.01 to 0.1 micron from the layer surface, and more preferably from about 0.02 to 0.08 micron from the layer surface. Preferably, the particles are situated at a distance of from about 0.005 to about 0.2 micron from each other, and more preferably at a distance of from about 0.05 to about 0.1 micron from each other, the distance being measured between the closest edges of the particles, i.e. from outer diameter to outer diameter. The migration marking material contiguous to the outer surface of the softenable layer is present in any effective amount, preferably from about 5 to about 80 percent by total weight of the softenable layer, and more preferably from about 25 to about 80 percent by total weight of the softenable layer, although the amount can be outside of this range.

Examples of suitable migration marking materials include selenium, alloys of selenium with alloying components such as tellurium, arsenic, antimony, thallium, bismuth, or mixtures thereof, selenium and alloys of selenium doped with halogens, as disclosed in, for example, U.S. Patent 3,312,548, and the like, phthalocyanines, and any other suitable materials as disclosed, for example, in U.S. Patent 3,975,195 directed to migration imaging members.

The migration imaging members can optionally contain a charge transport material. The charge transport material can be any suitable charge transport material either capable of acting as a softenable layer material or capable of being dissolved or dispersed on a molecular scale in the softenable layer material. When a charge transport material is also contained in another layer in the imaging member, preferably there is continuous transport of charge through the entire film structure. The charge transport material is defined as a material which is capable of improving the charge injection process for one sign of charge from the migration marking material into the softenable layer and also of transporting that charge through the softenable layer. The charge transport material can be either a hole transport material (transports positive charges) or an electron transport material (transports negative charges). The sign of the charge used to sensitize the migration imaging member during imaging can be of either polarity. Charge transporting materials are well known in the art. Typical charge transporting materials include the following:

Diamine transport molecules of the type described in U.S. Patent 4,306,008, U.S. Patent 4,304,829, U.S. Patent 4,233,384, U.S. Patent 4,115,116, U.S. Patent 4,299,897, and U.S. Patent 4,081,274. Typical diamine transport molecules include N,N'-diphenyl-N,N'-bis(3"-methylphenyl)-(1,1'-biphenyl)-4,4'-diamine, N,N'-diphenyl-N,N'-bis(4-methylphenyl)-(1,1'-biphenyl)-4,4'-diamine, N,N'-diphenyl-N,N'-bis(2-methylphenyl)-(1,1'-biphenyl)-4,4'-diamine, N,N'-diphenyl-N,N'-bis(3-ethylphenyl)-(1,1'-biphenyl)-4,4'-diamine, N,N'-diphenyl-N,N'-bis(4-ethylphenyl)-(1,1'-biphenyl)-4,4'-diamine, N,N'-diphenyl-N,N'-bis(4-n-butylphenyl)-(1,1'-biphenyl)-4,4'-diamine, N,N'-diphenyl-N,N'-bis(3-chlorophenyl)-[1,1'-biphenyl]-4,4'-diamine, N,N'-diphenyl-N,N'-bis(4-chlorophenyl)-[1,1'-biphenyl]-4,4'-diamine, N,N'-diphenyl-N,N'-bis(phenylmethyl)-[1,1'-biphenyl]-4,4'-diamine, N,N,N',N'-tetraphenyl-[2,2'-dimethyl-1,1'-biphenyl]-4,4'-diamine, N,N,N',N'-tetra-(4-methylphenyl)-[2,2'-dimethyl-1,1'-biphenyl]-4,4'-diamine, N,N'-diphenyl-N,N'-bis(4-methylphenyl)-[2,2'-dimethyl-1,1'-biphenyl]-4,4'-diamine, N,N'-diphenyl-N,N'-bis(2-methylphenyl)-[2,2'-dimethyl-1,1'-biphenyl]-4,4'- diamine, N,N'-diphenyl-N,N'-bis(3-methylphenyl)-[2,2'-dimethyl-1,1'-biphenyl]-4,4'-diamine, N,N'-diphenyl-N,N'-bis(3-methylphenyl)-pyrenyl-1,6-diamine, and the like.

Pyrazoline transport molecules as disclosed in U.S. Patent 4,315,982, U.S. Patent 4,278,746, and U.S. Patent 3,837,851. Typical pyrazoline transport molecules include 1-[lepidyl-(2)]-3-(p-diethylaminophenyl)-5-(p-diethylaminophenyl)pyrazoline, 1-[quinolyl-(2)]-3-(p-diethylaminophenyl)-5-(p-diethylaminophenyl)pyrazoline, 1-[pyridyl-(2)]-3-(p-diethylaminostyryl)-5-(p-diethylaminophenyl)pyrazoline, 1-[6-methoxypyridyl-(2)]-3-(p-diethylaminostyryl)-5-(p-diethylaminophenyl) pyrazoline, 1-phenyl-3-[p-dimethylaminostyryl]-5-(p-dimethylaminostyryl)pyrazoline, 1-phenyl-3-[p-diethylaminostyryl]-5-(p-diethylaminostyryl)pyrazoline, and the like.

Substituted fluorene charge transport molecules as described in U.S. Patent 4,245,021. Typical fluorene charge transport molecules include 9-(4'-dimethylaminobenzylidene)fluorene, 9-(4'-methoxybenzylidene)fluorene, 9-(2',4'-dimethoxybenzylidene)fluorene, 2-nitro-9-benzylidenefluorene,2-nitro-9-(4'-diethylaminobenzylidene)fluorene, and the like.

Oxadiazole transport molecules such as 2,5-bis(4-diethylaminophenyl)-1,3,4-oxadiazole, pyrazoline, imidazole, triazole, and the like. Other typical oxadiazole transport molecules are described, for example, in German Patent 1,058,836, German Patent 1,060,260, and German Patent 1,120,875.

Hydrazone transport molecules, such as p-diethylamino benzaldehyde(diphenylhydrazone), o-ethoxy-p-diethylaminobenzaldehyde-(diphenylhydrazone), o-methyl-p-diethylaminobenzaldehyde-(diphenylhydrazone), o-methyl-p-dimethylaminobenzaldehyde-(diphenylhydrazone), 1-naphthalenecarbaldehyde 1-methyl-1-phenylhydrazone, 1-naphthalenecarbaldehyde 1,1-phenylhydrazone, 4-methoxynaphthlene-1-carbaldeyde 1-methyl-1-phenylhydrazone, and the like. Other typical hydrazone transport molecules are described, for example in U.S. Patent 4,150,987, U.S. Patent 4,385,106, U.S. Patent 4,338,388, and U.S. Patent 4,387,147.

Carbazole phenyl hydrazone transport molecules such as 9-methylcarbazole-3-carbaldehyde-1,1-diphenylhydrazone, 9-ethylcarbazole-3-carbaldehyde-1-methyl-1-phenylhydrazone, 9-ethylcarbazole-3-carbaldehyde-1-ethyl-1-phenylhydrazone, 9-ethylcarbazole-3-carbaldehyde-1-ethyl-1-benzyl-1-phenylhydrazone, 9-ethylcarbazole-3-carbaldehyde-1,1-diphenylhydrazone, and the like. Other typical carbazole phenyl hydrazone transport molecules are described, for example, in U.S. Patent 4,256,821 and U.S. Patent 4,297,426.

Vinyl-aromatic polymers such as polyvinyl anthracene, polyacenaphthylene; formaldehyde condensation products with various aromatics such as condensates of formaldehyde and 3-bromopyrene; 2,4,7-trinitrofluorenone, and 3,6-dinitro-N-t-butylnaphthalimide as described, for example, in U.S. Patent 3,972,717.

Oxadiazole derivatives such as 2,5-bis-(p-diethylaminophenyl)-oxadiazole-1,3,4 described in U.S. Patent 3,895,944.

Tri-substituted methanes such as alkyl-bis(N,N-dialkylaminoaryl)methane, cycloalkyl-bis(N,N-dialkylaminoaryl)methane, and cycloalkenyl-bis(N,N-dialkylaminoaryl)methane as described in U.S. Patent 3,820,989.

9-Fluorenylidene methane derivatives having the formula wherein X and Y are cyano groups or alkoxycarbonyl groups; A, B, and W are electron withdrawing groups independently selected from the group consisting of acyl, alkoxycarbonyl, nitro, alkylaminocarbonyl, and derivatives thereof; m is a number of from 0 to 2; and n is the number 0 or 1 as described in U.S. Patent 4,474,865. Typical 9-fluorenylidene methane derivatives encompassed by the above formula include (4-n-butoxycarbonyl-9-fluorenylidene)malonontrile, (4-phenethoxycarbonyl-9-fluorenylidene)malonontrile, (4-carbitoxy-9-fluorenylidene)malonontrile, (4-n-butoxycarbonyl-2,7-dinitro-9-fluorenylidene)malonate, and the like.

Other charge transport materials include poly-1-vinylpyrene, poly-9-vinylanthracene, poly-9-(4-pentenyl)-carbazole, poly-9-(5-hexyl)-carbazole, polymethylene pyrene, poly-1-(pyrenyl)-butadiene, polymers such as alkyl, nitro, amino, halogen, and hydroxy substitute polymers such as poly-3-amino carbazole, 1,3-dibromo-poly-N-vinyl carbazole, 3,6-dibromo-poly-N-vinyl carbazole, and numerous other transparent organic polymeric or non-polymeric transport materials as described in U.S. Patent 3,870,516. Also suitable as charge transport materials are phthalic anhydride, tetrachlorophthalic anhydride, benzil, mellitic anhydride, S-tricyanobenzene, picryl chloride, 2,4-dinitrochlorobenzene, 2,4-dinitrobromobenzene, 4-nitrobiphenyl, 4,4-2,4,6-trinitroanisole, trichlorotrinitrobenzene, trinitro-O-toluene, 4,6-dichloro-1,3-dinitrobenzene, 4,6-dibromo-1,3-dinitrobenzene, P-dinitrobenzene, chloranil, bromanil, and mixtures thereof, 2,4,7-trinitro-9-fluorenone, 2,4,5,7-tetranitrofluorenone, trinitroanthracene, dinitroacridene, tetracyanopyrene, dinitroanthraquinone, polymers having aromatic or heterocyclic groups with more than one strongly electron withdrawing substituent such as nitro, sulfonate, carboxyl, cyano, or the like, including polyesters, polysiloxanes, polyamides, polyurethanes, and epoxies, as well as block, graft, or random copolymers containing the aromatic moiety, and the like, as well as mixtures thereof, as described in U.S. Patent 4,081,274.

Also suitable are charge transport materials such as triarylamines, including tritolyl amine, of the formula and the like, as disclosed in, for example, U.S. Patent 3,240,597 and U.S. Patent 3,180,730, and substituted diarylmethane and triarylmethane compounds, including bis-(4-diethylamino-2-methylphenyl)phenylmethane, of the formula and the like, as disclosed in, for example, U.S. Patent 4,082,551, U.S. Patent 3,755,310, U.S. Patent 3,647,431, British Patent 984,965, British Patent 980,879, and British Patent 1,141,666.

When the charge transport molecules are combined with an insulating binder to form the softenable layer, the amount of charge transport molecule which is used can vary depending upon the particular charge transport material and its compatibility (e.g. solubility) in the continuous insulating film forming binder phase of the softenable matrix layer and the like. Satisfactory results have been obtained using between about 5 percent to about 50 percent by weight charge transport molecule based on the total weight of the softenable layer. A particularly preferred charge transport molecule is one having the general formula wherein X, Y and Z are selected from the group consisting of hydrogen, an alkyl group having from 1 to about 20 carbon atoms and chlorine, and at least one of X, Y and Z is independently selected to be an alkyl group having from 1 to about 20 carbon atoms or chlorine. If Y and Z are hydrogen, the compound can be named N,N'-diphenyl-N,N'-bis(alkylphenyl)-[1,1'-biphenyl]-4,4'-diamine wherein the alkyl is, for example, methyl, ethyl, propyl, n-butyl, or the like, or the compound can be N,N'-diphenyl-N,N'-bis(chlorophenyl)-[1,1'-biphenyl]-4,4'-diamine. Results can be obtained when the softenable layer contains between about 8 percent to about 40 percent by weight of these diamine compounds based on the total weight of the softenable layer. Optimum results are achieved when the softenable layer contains between about 16 percent to about 32 percent by weight of N,N'-diphenyl-N,N'-bis(3''-methylphenyl)-(1,1'-biphenyl)-4,4'-diamine based on the total weight of the softenable layer.

The charge transport material is present in the softenable material in any effective amount, typically from about 5 to about 50 percent by weight and preferably from about 8 to about 40 percent by weight, although the amount can be outside these ranges. Alternatively, the softenable layer can employ the charge transport material as the softenable material if the charge transport material possesses the necessary film-forming characteristics and otherwise functions as a softenable material. The charge transport material can be incorporated into the softenable layer by any suitable technique. For example, it can be mixed with the softenable layer components by dissolution in a common solvent. If desired, a mixture of solvents for the charge transport material and the softenable layer material can be employed to facilitate mixing and coating. The charge transport molecule and softenable layer mixture can be applied to the substrate by any conventional coating process. Typical coating processes include draw bar coating, spray coating, extrusion, dip coating, gravure roll coating, wire-wound rod coating, air knife coating, and the like.

The optional adhesive layer can include any suitable adhesive material. Typical adhesive materials include copolymers of styrene and an acrylate, polyester resin such as DuPont 49000 (available from E.I. duPont de Nemours Company), copolymer of acrylonitrile and vinylidene chloride, polyvinyl acetate, polyvinyl butyral and the like and mixtures thereof. The adhesive layer can have any thickness, typically from about 0.05 to about 1 micron, although the thickness can be outside of this range. When an adhesive layer is employed, it preferably forms a uniform and continuous layer having a thickness of about 0.5 micron or less to ensure satisfactory discharge during the imaging process. It can also optionally include charge transport molecules.

The optional charge transport layer can comprise any suitable film forming binder material. Typical film forming binder materials include styrene acrylate copolymers, polycarbonates, co-polycarbonates, polyesters, co-polyesters, polyurethanes, polyvinyl acetate, polyvinyl butyral, polystyrenes, alkyd substituted polystyrenes, styrene-olefin copolymers, styrene-co-n-hexylmethacrylate, an 80/20 mole percent copolymer of styrene and hexylmethacrylate having an intrinsic viscosity of 0.179 dl/gm; other copolymers of styrene and hexylmethacrylate, styrene-vinyltoluene copolymers, polyalpha-methylstyrene, mixtures thereof, and copolymers thereof. The above group of materials is not intended to be limiting, but merely illustrative of materials suitable as film forming binder materials in the optional charge transport layer. The film forming binder material typically is substantially electrically insulating and does not adversely chemically react during the imaging process. Although the optional charge transport layer has been described as coated on a substrate, in some embodiments, the charge transport layer itself can have sufficient strength and integrity to be substantially self supporting and can, if desired, be brought into contact with a suitable conductive substrate during the imaging process. As is well known in the art, a uniform deposit of electrostatic charge of suitable polarity can be substituted for a conductive layer. Alternatively, a uniform deposit of electrostatic charge of suitable polarity on the exposed surface of the charge transport spacing layer can be substituted for a conductive layer to facilitate the application of electrical migration forces to the migration layer. This technique of "double charging" is well known in the art. The charge transport layer is of any effective thickness, typically from about 1 to about 25 microns, and preferably from about 2 to about 20 microns, although the thickness can be outside these ranges.

Charge transport molecules suitable for the charge transport layer are described in detail hereinabove. The specific charge transport molecule utilized in the charge transport layer of any given imaging member can be identical to or different from the charge transport molecule employed in the adjacent softenable layer. Similarly, the concentration of the charge transport molecule utilized in the charge transport spacing layer of any given imaging member can be identical to or different from the concentration of charge transport molecule employed in the adjacent softenable layer. When the charge transport material and film forming binder are combined to form the charge transport spacing layer, the amount of charge transport material used can vary depending upon the particular charge transport material and its compatibility (e.g. solubility) in the continuous insulating film forming binder. Satisfactory results have been obtained using between about 5 percent and about 50 percent based on the total weight of the optional charge transport spacing layer, although the amount can be outside this range. The charge transport material can be incorporated into the charge transport layer by techniques similar to those employed for the softenable layer.

The optional charge blocking layer can be of various suitable materials, provided that the objectives of the present invention are achieved, including aluminum oxide, polyvinyl butyral, silane and the like, as well as mixtures thereof. This layer, which is generally applied by known coating techniques, is of any effective thickness, typically from about 0.05 to about 0.5 micron, and preferably from about 0.05 to about 0.1 micron. Typical coating processes include draw bar coating, spray coating, extrusion, dip coating, gravure roll coating, wire-wound rod coating, air knife coating and the like.

The optional overcoating layer can be substantially electrically insulating, or have any other suitable properties. The overcoating preferably is substantially transparent, at least in the spectral region where electromagnetic radiation is used for imagewise exposure step in the imaging process. The overcoating layer is continuous and preferably of a thickness up to about 1 to 2 microns. More preferably, the overcoating has a thickness of between about 0.1 and about 0.5 micron to minimize residual charge buildup. Overcoating layers greater than about 1 to 2 microns thick can also be used. Typical overcoating materials include acrylic-styrene copolymers, methacrylate polymers, methacrylate copolymers, styrene-butylmethacrylate copolymers, butylmethacrylate resins, vinylchloride copolymers, fluorinated homo or copolymers, high molecular weight polyvinyl acetate, organosilicon polymers and copolymers, polyesters, polycarbonates, polyamides, polyvinyl toluene and the like. The overcoating layer generally protects the softenable layer to provide greater resistance to the adverse effects of abrasion during handling and imaging. The overcoating layer preferably adheres strongly to the softenable layer to minimize damage. The overcoating layer can also have abhesive properties at its outer surface which provide improved resistance to toner filming during toning, transfer, and/or cleaning. The abhesive properties can be inherent in the overcoating layer or can be imparted to the overcoating layer by incorporation of another layer or component of abhesive material. These abhesive materials should not degrade the film forming components of the overcoating and preferably have a surface energy of less than about 20 ergs/cm². Typical abhesive materials include fatty acids, salts and esters, fluorocarbons, silicones, and the like. The coatings can be applied by any suitable technique such as draw bar, spray, dip, melt, extrusion or gravure coating. It will be appreciated that these overcoating layers protect the imaging member before imaging, during imaging, after the members have been imaged.

As illustrated schematically in Figure 2, migration imaging member 11 comprises in the order shown a substrate 12, an optional adhesive layer 13 situated on substrate 12, an optional charge blocking layer 14 situated on optional adhesive layer 13, an optional charge transport layer 15 situated on optional charge blocking layer 14, a softenable layer 16 situated on optional charge transport layer 15, said softenable layer 16 comprising softenable material 17, charge transport material 18, and migration marking material 19 situated at or near the surface of the layer spaced from the substrate, and an infrared or red light radiation sensitive layer 20 situated on softenable layer 16 comprising infrared or red light radiation sensitive pigment particles 21 optionally dispersed in polymeric binder 22. Alternatively (not shown), infrared or red light radiation sensitive layer 20 can comprise infrared or red light radiation sensitive pigment particles 21 directly deposited as a layer by, for example, vacuum evaporation techniques or other coating methods. Optional overcoating layer 23 is situated on the surface of imaging member 11 spaced from the substrate 12.

As illustrated schematically in Figure 3, migration imaging member 24 comprises in the order shown a substrate 25, an optional adhesive layer 26 situated on substrate 25, an optional charge blocking layer 27 situated on optional adhesive layer 26, an infrared or red light radiation sensitive layer 28 situated on optional charge blocking layer 27 comprising infrared or red light radiation sensitive pigment particles 29 optionally dispersed in polymeric binder 30, an optional charge transport layer 31 situated on infrared or red light radiation sensitive layer 28, and a softenable layer 32 situated on optional charge transport layer 31, said softenable layer 32 comprising softenable material 33, charge transport material 34, and migration marking material 35 situated at or near the surface of the layer spaced from the substrate. Optional overcoating layer 36 is situated on the surface of imaging member 24 spaced from the substrate 25.

The infrared or red light sensitive layer generally comprises a pigment sensitive to infrared and/or red light radiation. While the infrared or red light sensitive pigment may exhibit some photosensitivity in the wavelength to which the migration marking material is sensitive, it is preferred that photosensitivity in this wavelength range be minimized so that the migration marking material and the infrared or red light sensitive pigment exhibit absorption peaks in distinct, different wavelength regions. This pigment can be deposited as the sole or major component of the infrared or red light sensitive layer by any suitable technique, such as vacuum evaporation or the like. An infrared or red light sensitive layer of this type can be formed by placing the pigment and the imaging member comprising the substrate and any previously coated layers into an evacuated chamber, followed by heating the infrared or red light sensitive pigment to the point of sublimation. The sublimed material recondenses to form a solid film on the imaging member. Alternatively, the infrared or red light sensitive pigment can be dispersed in a polymeric binder and the dispersion coated onto the imaging member to form a layer. Examples of suitable red light sensitive pigments include perylene pigments such as benzimidazole perylene, dibromoanthranthrone, crystalline trigonal selenium, beta-metal free phthalocyanine, azo pigments, and the like, as well as mixtures thereof. Examples of suitable infrared sensitive pigments include X-metal free phthalocyanine, metal phthalocyanines such as vanadyl phthalocyanine, chloroindium phthalocyanine, titanyl phthalocyanine, chloroaluminum phthalocyanine, copper phthalocyanine, magnesium phthalocyanine, and the like, squaraines, such as hydroxy squaraine, and the like as well as mixtures thereof. Examples of suitable optional polymeric binder materials include polystyrene, styrene-acrylic copolymers, such as styrene-hexylmethacrylate copolymers, styrene-vinyl toluene copolymers, polyesters, such as PE-200, available from Goodyear, polyurethanes, polyvinylcarbazoles, epoxy resins, phenoxy resins, polyamide resins, polycarbonates, polyterpenes, silicone elastomers, polyvinylalcohols, such as Gelvatol 20-90, 9000, 20-60, 6000, 20-30, 3000, 40-20, 40-10, 26-90, and 30-30, available from Monsanto Plastics and Resins Co., St. Louis, MO, polyvinylformals, such as Formvar 12/85, 5/95E, 6/95E, 7/95E, and 15/95E, available from Monsanto Plastics and Resins Co., St. Louis, MO, polyvinylbutyrals, such as Butvar B-72, B-74, B-73, B-76, B-79, B-90, and B-98, available from Monsanto Plastics and Resins Co., St. Louis, MO, Zeneca resin A622, available from Zeneca Colours, Wilmington, DE, and the like as well as mixtures thereof. When the infrared or red light sensitive layer comprises both a polymeric binder and the pigment, the layer typically comprises the binder in an amount of from about 5 to about 95 percent by weight and the pigment in an amount of from about 5 to about 95 percent by weight although the relative amounts can be outside this range. Preferably, the infrared or red light sensitive layer comprises the binder in an amount of from about 40 to about 90 percent by weight and the pigment in an amount of from about 10 to about 60 percent by weight. Optionally, the infrared sensitive layer can contain a charge transport material as described herein when a binder is present; when present, the charge transport material is generally contained in this layer in an amount of from about 5 to about 30 percent by weight of the layer. The optional charge transport material can be incorporated into the infrared or red light radiation sensitive layer by any suitable technique. For example, it can be mixed with the infrared or red light radiation sensitive layer components by dissolution in a common solvent. If desired, a mixture of solvents for the charge transport material and the infrared or red light sensitive layer material can be employed to facilitate mixing and coating. The infrared or red light radiation sensitive layer mixture can be applied to the substrate by any conventional coating process. Typical coating processes include draw bar coating, spray coating, extrusion, dip coating, gravure roll coating, wire-wound rod coating, air knife coating, and the like. An infrared or red light sensitive layer wherein the pigment is present in a binder can be prepared by dissolving the polymer binder in a suitable solvent, dispersing the pigment in the solution by ball milling, coating the dispersion onto the imaging member comprising the substrate and any previously coated layers, and evaporating the solvent to form a solid film. When the infrared or red light sensitive layer is coated directly onto the softenable layer containing migration marking material, preferably the selected solvent is capable of dissolving the polymeric binder for the infrared or red sensitive layer but does not dissolve the softenable polymer in the layer containing the migration marking material. One example of a suitable solvent is isobutanol with a polyvinyl butyral binder in the infrared or red sensitive layer and a styrene/ethyl acrylate/acrylic acid terpolymer softenable material in the layer containing migration marking material. The infrared or red light sensitive layer can be of any effective thickness. Typical thicknesses for infrared or red light sensitive layers comprising a pigment and a binder are from about 0.05 to about 2 microns, and preferably from about 0.1 to about 1.5 microns, although the thickness can be outside these ranges. Typical thicknesses for infrared or red light sensitive layers consisting of a vacuum-deposited layer of pigment are from about 200 to about 2,000 Angstroms, and preferably from about 300 to about 1,000 Angstroms, although the thickness can be outside these ranges.

The transparentizing agent can be contained in any of the migration imaging member layers so that upon migration of the migration marking material through the softenable layer, either the migrated particles or the unmigrated particles are selectively transparentized by the transparentizing agent. For example, in the embodiment illustrated in Figure 1, when the optional adhesive layer 3, optional charge blocking layer 4, and optional charge transport layer 5 are all absent, the transparentizing agent can be contained in part or all of the substrate layer 2. Upon migration of the migration marking material 8 through the softenable layer 6, migrated particles contact the transparentizing agent in substrate 2 and become transparentized, thereby reducing the Dₘᵢₙ value of the imaging member subsequent to development. When one or more of the optional layers is present, the transparentizing agent can be present in one or more of these layers so that upon migration of the migration marking material 8 through the softenable layer 6, migrated particles contact the transparentizing agent in one or more of the optional layers and become transparentized, thereby reducing the Dₘᵢₙ value of the imaging member subsequent to development. Further, in the embodiment illustrated in Figure 2, when the optional adhesive layer 13, optional charge blocking layer 14, and optional charge transport layer 15 are all absent, the transparentizing agent can be contained in part or all of the substrate layer 12. Upon migration of the migration marking material 19 through the softenable layer 16, migrated particles contact the transparentizing agent in substrate 12 and become transparentized, thereby reducing the Dₘᵢₙ value of the imaging member subsequent to development. When one or more of the optional layers is present, the transparentizing agent can be present in one or more of these layers so that upon migration of the migration marking material 19 through the softenable layer 16, migrated particles contact the transparentizing agent in one or more of the optional layers and become transparentized, thereby reducing the Dₘᵢₙ value of the imaging member subsequent to development. Additionally, in the embodiment illustrated in Figure 3, when the optional adhesive layer 26, optional charge blocking layer 27, and optional charge transport layer 31 are all absent, the transparentizing agent can be contained in part or all of the infrared or red light sensitive layer 28. Upon migration of the migration marking material 35 through the softenable layer 32, migrated particles contact the transparentizing agent in infrared or red light sensitive layer 28 and become transparentized, thereby reducing the Dₘᵢₙ value of the imaging member subsequent to development. When one or more of the optional layers is present, the transparentizing agent can be present in one or more of these layers, such as charge transport layer 31, so that upon migration of the migration marking material 35 through the softenable layer 32, migrated particles contact the transparentizing agent in one or more of the optional layers and become transparentized, thereby reducing the Dₘᵢₙ value of the imaging member subsequent to development.

The transparentizing agent can also be present in the softenable layer itself. For example, in the embodiment illustrated in Figure 1, the transparentizing agent can be present in softenable layer 6; in the embodiment illustrated in Figure 2, the transparentizing agent can be present in softenable layer 16; in the embodiment illustrated in Figure 3, the transparentizing agent can be present in softenable layer 32. When present in the softenable layer, the transparentizing agent can be contained throughout the softenable layer without being uniformly distributed therein. For example, the transparentizing agent can be situated or concentrated near the bottom of the softenable layer (i.e., that part of the softenable layer in closest proximity to the substrate) so that subsequent to image formation and development, migrated migration marking particles contact the transparentizing agent and become transparentized, while unmigrated migration marking particles contact the transparentizing agent either not at all or in a manner such that the concentration of transparentizing agent contacting the unmigrated marking particles is less than the concentration of transparentizing agent contacting the migrated marking particles. Further, the transparentizing agent can be situated or concentrated near the top of the softenable layer (i.e., that part of the softenable layer spaced from the substrate) so that subsequent to image formation and development, unmigrated migration marking particles contact the transparentizing agent and become transparentized, while migrated migration marking particles contact the transparentizing agent either not at all or in a manner such that the concentration of transparentizing agent contacting the migrated marking particles is less than the concentration of transparentizing agent contacting the unmigrated marking particles. The concentration of transparentizing agent within the softenable layer can be varied according to depth within the layer by any suitable method, such as by applying the softenable layer by a series of solvent coating steps, wherein the concentration of transparentizing agent dispersed with the softenable material and solvent is varied to increase or decrease the concentration of transparentizing agent as successive coatings are applied. Thereafter, the migration marking material is applied to the softenable layer by any suitable or desired method, such as solvent coating, evaporation coating, or the like.

The transparentizing agent can further be present in a separate layer or coating within the migration imaging member structure. For example, as illustrated schematically in Figure 4, migration imaging member 40 comprises a substrate 41, an optional adhesive layer 42 situated on the substrate 41, an optional charge blocking layer 43 situated on optional adhesive layer 42, an optional charge transport layer 44 situated on optional charge blocking layer 43, a transparentizing layer 45 situated on optional charge transport layer 44, and a softenable layer 46 situated on transparentizing layer 45, said softenable layer 46 comprising softenable material 47, migration marking material 48 situated at or near the surface of the layer spaced from the substrate, and optional charge transport material 49 dispersed throughout softenable material 47. Optional overcoating layer 50 is situated on the surface of softenable layer 46 spaced from the substrate 41. Any or all of the optional layers and materials can be absent from the imaging member. In addition, any of the optional layers present need not be in the order shown, but can be in any suitable arrangement. For example, if the optional adhesive layer 42, optional charge blocking layer 43, and optional charge transport layer 44 are absent, transparentizing layer 46 is coated directly onto substrate 41 and is situated between and in contact with substrate 41 and softenable layer 46.

Similarly, in the embodiment illustrated in Figure 5, migration imaging member 51 comprises in the order shown a substrate 52, an optional adhesive layer 53 situated on substrate 52, an optional charge blocking layer 54 situated on optional adhesive layer 53, an optional charge transport layer 55 situated on optional charge blocking layer 54, a transparentizing layer 56 situated on optional charge transport layer 55, a softenable layer 57 situated on transparentizing layer 56, said softenable layer 57 comprising softenable material 58, charge transport material 59, and migration marking material 60 situated at or near the surface of the layer spaced from the substrate, and an infrared or red light radiation sensitive layer 61 situated on softenable layer 57 comprising infrared or red light radiation sensitive pigment particles 62 optionally dispersed in polymeric binder 63. Alternatively (not shown), infrared or red light radiation sensitive layer 61 can comprise infrared or red light radiation sensitive pigment particles 62 directly deposited as a layer by, for example, vacuum evaporation techniques or other coating methods. Optional overcoating layer 64 is situated on the surface of imaging member 51 spaced from the substrate 52. Any or all of the optional layers and materials can be absent from the imaging member. In addition, any of the optional layers present need not be in the order shown, but can be in any suitable arrangement. For example, if the optional adhesive layer 53, optional charge blocking layer 54, and optional charge transport layer 55 are absent, transparentizing layer 56 is coated directly onto substrate 52 and is situated between and in contact with substrate 52 and softenable layer 57.

Similarly, as illustrated schematically in Figure 6, migration imaging member 65 comprises in the order shown a substrate 66, an optional adhesive layer 67 situated on substrate 66, an optional charge blocking layer 68 situated on optional adhesive layer 67, an infrared or red light radiation sensitive layer 69 situated on optional charge blocking layer 68 comprising infrared or red light radiation sensitive pigment particles 70 optionally dispersed in polymeric binder 71, an optional charge transport layer 72 situated on infrared or red light radiation sensitive layer 69, a transparentizing layer 73 situated on optional charge transport layer 72, and a softenable layer 74 situated on transparentizing layer 73, said softenable layer 74 comprising softenable material 75, charge transport material 76, and migration marking material 77 situated at or near the surface of the layer spaced from the substrate. Optional overcoating layer 78 is situated on the surface of imaging member 65 spaced from the substrate 66. Any or all of the optional layers and materials can be absent from the imaging member. In addition, any of the optional layers present need not be in the order shown, but can be in any suitable arrangement. For example, if the optional adhesive layer 67, optional charge blocking layer 68, and optional charge transport layer 72 are absent, transparentizing layer 73 is coated directly onto infrared or red light sensitive layer 69 and is situated between and in contact with infrared or red light sensitive layer 69 and softenable layer 74.

In the embodiments illustrated in Figures 4, 5, and 6, the transparentizing layer is situated below the softenable layer (i.e., is situated between the softenable layer and the substrate), so that subsequent to image formation and development, migrated migration marking particles contact the transparentizing agent in the transparentizing layer and become transparentized, while unmigrated migration marking particles do not contact the transparentizing agent in the transparentizing layer and thus are not transparentized. The transparentizing agent can also be situated above the softenable layer (i.e., situated so that the softenable layer is between the transparentizing layer and the substrate). For example, as illustrated schematically in Figure 7, migration imaging member 79 comprises a substrate 80, an optional adhesive layer 81 situated on the substrate 80, an optional charge blocking layer 82 situated on optional adhesive layer 81, an optional charge transport layer 83 situated on optional charge blocking layer 82, a softenable layer 84 situated on optional charge transport layer 83, said softenable layer 84 comprising softenable material 85, migration marking material 86 situated at or near the surface of the layer spaced from the substrate, and optional charge transport material 87 dispersed throughout softenable material 85, and a transparentizing layer 88 situated on softenable layer 84. Optional overcoating layer 89 is situated on the surface of transparentizing layer 88 spaced from the substrate 80. Any or all of the optional layers and materials can be absent from the imaging member. In addition, any of the optional layers present need not be in the order shown, but can be in any suitable arrangement.

Similarly, in the embodiment illustrated in Figure 8, migration imaging member 90 comprises in the order shown a substrate 91, an optional adhesive layer 92 situated on substrate 91, an optional charge blocking layer 93 situated on optional adhesive layer 92, an optional charge transport layer 94 situated on optional charge blocking layer 93, a softenable layer 95 situated on optional charge transport layer 94, said softenable layer 95 comprising softenable material 96, charge transport material 97, and migration marking material 98 situated at or near the surface of the layer spaced from the substrate, a transparentizing layer situated on softenable layer 95, and an infrared or red light radiation sensitive layer 100 situated on transparentizing layer 99 comprising infrared or red light radiation sensitive pigment particles 101 optionally dispersed in polymeric binder 102. Alternatively (not shown), infrared or red light radiation sensitive layer 100 can comprise infrared or red light radiation sensitive pigment particles 101 directly deposited as a layer by, for example, vacuum evaporation techniques or other coating methods. Optional overcoating layer 103 is situated on the surface of imaging member 90 spaced from the substrate 91. Any or all of the optional layers and materials can be absent from the imaging member. In addition, any of the optional layers present need not be in the order shown, but can be in any suitable arrangement.

Similarly, as illustrated schematically in Figure 9, migration imaging member 104 comprises in the order shown a substrate 105, an optional adhesive layer 106 situated on substrate 105, an optional charge blocking layer 107 situated on optional adhesive layer 106, an infrared or red light radiation sensitive layer 108 situated on optional charge blocking layer 107 comprising infrared or red light radiation sensitive pigment particles 109 optionally dispersed in polymeric binder 110, an optional charge transport layer 111 situated on infrared or red light radiation sensitive layer 108, a softenable layer 112 situated on optional charge transport layer 111, said softenable layer 112 comprising softenable material 113, charge transport material 114, and migration marking material 115 situated at or near the surface of the layer spaced from the substrate, and transparentizing layer 116 situated on softenable layer 112. Optional overcoating layer 117 is situated on the surface of imaging member 104 spaced from the substrate 105. Any or all of the optional layers and materials can be absent from the imaging member. In addition, any of the optional layers present need not be in the order shown, but can be in any suitable arrangement.

In embodiments of the present invention wherein two or more softenable layers, each containing a migration marking material, are present in the migration imaging member, the transparentizing agent can be present within one or both of the softenable layers as illustrated schematically in Figures 1 through 3. Additionally, the transparentizing agent can be present as a separate layer as illustrated in Figures 4 through 9. Further, the transparentizing agent can be present as a separate layer situated between the two softenable layers, as illustrated schematically in Figure 10. As illustrated schematically in Figure 10, migration imaging member 118 comprises in the order shown a substrate 119, an optional adhesive layer 120 situated on substrate 119, an optional charge blocking layer 121 situated on optional adhesive layer 120, an optional charge transport layer 122 situated on optional charge blocking layer 121, a first softenable layer 123 situated on optional charge transport layer 122, said first softenable layer 123 comprising first softenable material 124, optional first charge transport material 125, and first migration marking material 126 situated at or near the surface of the first softenable layer spaced from the substrate, a transparentizing layer 127 situated on first softenable layer 123, and a second softenable layer 128 situated on transparentizing layer 127 comprising second softenable material 129, optional second charge transport material 130, and second migration marking material 131 situated at or near the surface of second softenable layer 128 in contact with transparentizing layer 127. Alternatively (not shown), second migration marking material can be situated at or near the surface of second softenable layer 128 spaced from substrate 119, or can be dispersed uniformly within second softenable layer 128. Optional overcoating layer 132 is situated on the surface of the imaging member spaced from the substrate 119. Further (not shown), an infrared or red light sensitive layer can be situated within the migration imaging member having two softenable layers in configurations as illustrated, for example, in Figures 2, 3, 5, 6, 8, and 9.

The transparentizing layer as illustrated in Figures 4 through 10 can be applied to the imaging member by any desired or suitable method. For example, a layer of softenable material (either the same as or different from the softenable material employed in the softenable layer) can be prepared by admixing the softenable material and the transparentizing agent and applying the mixture to the imaging member by any desired method, such as draw bar coating, spray coating, extrusion, dip coating, gravure roll coating, wire-wound rod coating, air knife coating and the like. Alternatively, the transparentizing agent can be coated directly onto the underlying layer in the migration imaging member, with no need for a binder or matrix, by dissolving or dispersing the transparentizing agent into a solvent, coating the solution or dispersion onto the underlying layer, and allowing the solvent to evaporate. For transparentizing agents suitable for evaporation coating techniques, the transparentizing agent can be vacuum evaporated onto the underlying layer of the migration imaging member. When the transparentizing agent is incorporated into another layer of the migration imaging member, or when the transparentizing agent is admixed with a binder and/or any additional materials to form a separate transparentizing layer within the migration imaging member, the transparentizing agent preferably is present within the layer in an amount of from about 1 to about 50 percent by weight, and more preferably 5 to about 20 percent by weight, although the amount can be outside these ranges. When the transparentizing agent is present in a separate transparentizing layer, preferably the layer is of a thickness of from about 2 to about 4 microns, although the thickness can be outside this range.

The transparentizing agent preferably is a monomeric material. In some instances, oligomeric materials (i.e., molecules having up to about four repeating monomer units) can also be employed as the transparentizing agent. Some polymeric materials may also be suitable if they contain some functional groups similar to those contained in suitable monomeric or oligomeric materials. While not being limited to any particular theory, it is believed that the transparentizing agent may chelate with the migration marking material, thereby rendering it transparent, or may enhance the ability of the migration marking material to agglomerate, or may oxidize the migration marking material, thereby rendering it transparent.

Examples of transparentizing agents suitable for the present invention include the following:

I. Azacyclic and azaheterocyclic compounds, including (A) piperidines and piperidine derivatives, including those of the general formulae: wherein R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈, and R₃₉ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈, and R₃₉ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable piperadine compounds and derivatives include (1) homopiperidine, (2) piperidinethiocyanate, (3) (±)-2-piperidinemethanol, (4) 3-piperidinemethanol, (5) 2-piperidineethanol, (6) 4-piperidineethanol, (7) 4-piperidine monohydrate hydrochloride, (8) 1-aminopiperidine, (9) 1-(2-aminoethyl)piperidine,(10) 4-(aminomethyl)piperidine, (11) 3-piperidino-1,2-propanediol, (12) 1-piperidine propionic acid, (13) 1-methyl-4-(methylamino)piperidine, (14) 1-acetyl-3-methylpiperidine, (15) 4'-piperidinoacetophenone, (16) 4-phenylpiperidine, (17) 4-piperidinopiperidine, (18) 4-benzylpiperidine, (19) 4-(4-methylpiperidino)pyridine, (20) 4-piperidone ethylene ketal, (21) bis(pentamethylene)urea, (22) 1-benzyl-4-hydroxypiperidine, (23) 1-benzoyl-4-piperidone, (24) 1,1'-methylenebis(3-methylpiperidine), (25) 4,4'-trimethylenedipiperidine, (26) 4,4'-trimethylenebis(1-menthylpiperidine), (27) 4,4'-trimethylenebis(1-piperidinepropionitrile), (28) 4,4'-trimethylenebis(1-piperidineethanol), (29) 2,2,6,6-tetramethylpiperidine, (30) 4-amino-2,2,6,6-tetramethylpiperidine, (31) 4-(dimethylamino)-1,2,2,6,6-pentamethylpiperidine, (32) N,N'-bis(2,2,6,6-tetramethyl-4-piperidinyl)-1,6-hexanediamine, (33) tripiperidinophosphine oxide, (34) tropane, (35) tropinehydrate, (36) tropinone, (37) 8-hydroxytropinone, (38) 2-piperidine carboxylic acid, (39) 2-piperidone, (40) 4,4'-trimethylene bis (1-piperidine carboxamide), (41) 4-methyl-2-(piperidinomethyl) phenol, (42) 1-methyl-4-piperidinyl bis (chlorophenoxy) acetate, (43) 2-(hexamethylene imino) ethyl chloride monohydrochloride, (44) 3-(hexahydro-1H-azepin-1-yl)-3'-nitropropiophenone hydrochloride, (45) imipramine hydrochloride [5-(3-dimethyl aminopropyl)-10,11-dihydro 5H-dibenz-(b,f) azepine hydrochloride], (46) carbamezepine [5H-dibenzo (b,f)-azepine-5-carboxamide], (47) 5,6,11,12-tetrahydro dibenz [b,f] azocine hydrochloride, (48) quinuclidine hydrochloride, (49) 3-quinuclidinol hydrochloride, (50) 3-quinuclidinone hydrochloride, (51) 2-methylene-3-quinuclidinone dihydrate hydrochloride, (52) 3-amino quinuclidine dihydrochloride, (53) 3-chloro quinuclidine hydrochloride, (54) quinidine sulfate dihydrate, (55) quinine monohydrochloride dihydrate, (56) quinine sulfate monohydrate, (57) hydroquinidine hydrochloride, (58) hydroquinine hydrobromide dihydrate, and the like;

(B) piperazines and piperazine derivatives, including those of the general formulae wherein R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, and R₂₂ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ and R₂₂ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, IO₃⁻, ClO₃⁻, or the like, as well as mixtures thereof.

Examples of suitable piperazine compounds and derivatives include (1) piperazine and piperazine hexahydrate, (2) homopiperazine, (3) 1-methylpiperazine, (4) 2-methylpiperazine, (5) 1-acetylpiperazine, (6) 1-(2-hydroxyethyl)piperazin, (7) 1-(2-aminoethyl)piperazine, (8) tert-butyl 1-piperazinecarboxylate, (9) N-isopropyl-1-piperazineacetamide, (10) 1-(2-methoxyphenyl)piperazine, (11) 1-(2-pyridyl)piperazine, (12) 1-benzylpiperazine, (13) 1-cinnamylpiperazine, (14) 1-(4-chlorobenzhydryl)piperazine, (15) 2,6-dimethylpiperazine, (16) 1-amino-4-methylpiperazine, (17) 1-amino-4-(2-hydroxyethyl)piperazine, (18) 1,4-bis(2-hydroxyethyl)piperazine, (19) 1,4-bis(3-aminopropyl)piperazine, (20) tert-butyl-4-benzyl-1-piperazinecarboxylate, (21) 1-piperonyl piperazine, (22) bis(4-methyl-1-homopiperazinylthio-carbonyl)disulfide, (23) 1-amino-4-methyl piperazine dihydrochloride monohydrate, (24) 1-(3-chloropropyl)-piperazine dihydrochloride monohydrate, (25) 1-(2,3-xylyl) piperazine monohydrochloride, (26) 1,1-dimethyl-4-phenyl piperazineium iodide, and the like;

(C) cyclic compounds wherein the ring contains three nitrogen atoms, including (1) 1,4,7-triazacyclononane,(2) 1,5,9-triazacyclododecane,(3) triazoles and triazole derivatives, including those of the general formulae wherein R₁, R₂, and R₃ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, and R₃ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof, such as (a) 1,2,3-triazole,(b) 4-amino-1,2,4-triazole, (c) 3-amino-5-methylthio-lH-1,2,4-triazole, (d) benzotriazole, (e) 1-aminobenzotriazole, (f) 1-cyanobenzotriazole, (g) 5-methyl-1H-benzotriazole, (h) 1H-benzotriazole-1-ylmethyl isocyanide, (i) 2-[3-(2H-benzotriazole-2-yl)-4-hydroxyphenyl]ethyl methacrylate, (j) 1,2,4-triazole, (k) 1,2,4-triazole sodium derivative, (I) 3-amino-1,2,4-triazole, (m) 3,5-diamino-1,2,4-triazole, (n) 3-amino-5-mercapto-1,2,4-triazole, (o) 3-amino-1,2,4-triazole-5-carboxylic acid hemihydrate, (p) 4-amino-3-hydrazino-5-mercapto-1,2,4-triazole, (q) 1,2,3-triazole-4,5-dicarboxylic acid monohydrate, (r) nitron [4,5-dihydro-2,4-diphenyl-5-(phenylimino)-1H-1,2,4-triazolium hydroxide inner salt], (s) 1-hydroxybenzotriazole hydrate, and the like; (4) triazines and triazine derivatives, including those of the general formulae wherein R₁, R₂, R₃, R₄, R₅, R₆, R₇, R₈, R₉, R₁₀, R₁₁, and R₁₂ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, and R₁₂ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃-, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof, such as (a) 1,3,5-triazine, (b) cyanuric acid, (c) trithiocyanuric acid, (d) 2,4-bis (methylthio)-6-chloro-1,3,5-triazine, (e) 2-chloro-4,6-dimethoxy-1,3,5-triazine, (f) 2-chloro-4,6-diamino-1,3,5-triazine, (g) trichloromelamine, (h) cyanuric chloride, (i) 2,4,6-tris(perfluoroheptyl)-1,3,5-triazine, (j) hexahydro-2,4,6-trimethyl-1,3,5-triazine trihydrate, (k) 1,3,5-trimethylhexahydro-1,3,5-triazine, (I) 1,3,5-triethylhexahydro-1,3,5-triazine, (m) 1,3,5-triclohexylhexahydro-1,3,5-triazine, (n) 1,3,5-tribenzylhexahydro-1,3,5-triazine, (o) trichloroisocyanuric acid, (p) tris (2,3-dibromopropylisocyanurate), (q) cyanuric acid compound with melamine, and the like; (5) urazoles and urazole derivatives, including those of the general formulae wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof, such as (a) urazole, (b) 1-methyl urazole, (c) 4-phenyl urazole, (d) D,L-5-(4-hydroxyphenyl)-5-phenyl hydantoin, (e) β-tetralone hydantoin, and the like;

(D) cyclic compounds wherein the ring contains four nitrogen atoms, including (1) cyclen (1,4,7,10-tetraazacyclododecane), (2) 1,4,8,11-tetraazacyclotetradecane, (3) 1,4,8,11-tetramethyl- 1,4,8,11 1,4,8,11 -tetraazacyclotetradecane, (4) 1,4,8,11-tetraazacyclotetradecane-5,7-dione, (5) 1,4,8,12-tetraazacyclopentadecane, (6) porphines and porphine derivatives, including those of the general formula wherein R₁, R₂, R₃, R₄, R₅, R₆, R₇, R₈, R₉, R₁₀, R₁₁, R₁₂, R₁₃, and R₁₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, and R₁₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃-, SO₃²⁻, BrO₃⁻, lO₃⁻, ClO₃⁻, or the like, as well as mixtures thereof. Examples of suitable porphines and porphine derivatives include (a) 2,3,7,8,12,13,17,18-octaethyl-21H,23H-porphine, (b) dimethyl 3,7,12,17-tetramethyl-21H,23H-porphine-2,18-dipropionate, (c) dimethyl 7,12-diacetyl-3,8,13,17-tetramethyl-21H,23H-porphine-2,18-dipropionate, (d) 8,3-divinyl-3,7,12,17-tetramethyl-21H,23H-porphine-2,18-dipropionic acid, disodium salt, (e) 5,10,15,20-tetraphenyl-21H,23H-porphine, (f) 5,10,1 5,20-tetrakis(4-methoxyphenyl)-21H,23H-porphine, (g) 5,10,15-20-tetrakis[4-(trimethylamino)phenyl]-21H,23H-porphine tetra-p-tosylate salt, (h) 5,10,15,20-tetra(4-pyridyl)-21H,23H-porphine, (i) 5,10,15,20-tetrakis(1-methyl-4-pyridyl)-21H,23H-porphine, tetra-p-tosylate salt), and the like; (7) tetrazoles and tetrazole derivatives, including those of the general formula wherein R₁ and R₂ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R1 and R2 can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, CIO₃⁻, or the like, as well as mixtures thereof, including (a) 1,5-pentamethylenetetrazole, (b) 1-H-tetrazole, (c) 5-amino tetrazole monohydrate, (d) 2,3,5-triphenyl-2H-tetrazolium chloride, (e) 2-(4-iodophenyl)-5-(4-nitrophenyl)-3-phenyltetrazolium chloride, (f) 1,2,3,3-tetramethyl-3H-indolinium iodide, and the like;

(E) cyclic compounds wherein the ring contains six nitrogen atoms, including (1) hexacyclen trisulfate, (2) hexamethylhexacyclen [1,4,7,10,13,16-hexamethyl-1,4,7,10,13-16-hexaazacyclooctadecane], and the like;

(F) pyrrole compounds, including those of the general formula wherein R₁, R₂, R₃, R₄, and R₅ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, and R₅ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof; and (G) pyrrolidine compounds, including those of the general formula wherein R₁, R₂, R₃, R₄, R₅, R₆, R₇, R₈, and R₉ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, and R₉ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between pyrrole or pyrrolidine and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable pyrrole and pyrrolidine compounds include (1) pyrrole-2-carboxaldehyde, (2) L-proline amide, (3) 3-pyrrolidino-1,2-propane diol, (4) 1-(pyrrolidino carbonylmethyl) piperazine, (5) 4-pyrrolidinopyridine, (6) 3-indolylacetonitrile, (7) 6-nitroindoline, (8) 7-azaindole, (9) indazole, (10) 2-acetyl-pyrrole, (11) 2-acetyl-1-methylpyrrole, (12) 3-acetyl-1 -methyl pyrrole, (13) 3-acetyl-2,4-dimethylpyrrole, (14) pyrrole-2-carboxylic acid, (15) 3-carboxy-1,4-dimethyl-2-pyrroleacetic acid, (16) proline, (17) 2-pyrrolidone-5-carboxylic acid, (18) 4-hydroxy-L-proline, (19) 1,1'-ethylene bis (5-oxo-3-pyrrolidine carboxylic acid), (20) kainic acid monohydrate (2-carboxy-4-isopropenyl-3-pyrrolidine acetic acid monohydrate), (21) 1-amino pyrrolidine hydrochloride, (22) 2-(2-chloroethyl)-1-methyl pyrrolidine hydrochloride, (23) 1-(2-chloroethyl) pyrrolidine hydrochloride, (24) tremorine dihydrochloride [1,1'-(2-butynylene) dipyrrolidine hydrochloride],(25) L-proline methyl ester hydrochloride, (26) ammonium pyrrolidine dithiocarbamate, (27) pyrrolidone hydrotribromide, (28) 1-(4-chlorobenzyl)-2-(1-pyrrolidinyl methyl) benzimidazole hydrochloride, (29) billverdin dihydrochloride, (30) indole, (31) 4,5,6,7-tetrahydroindole, (32) 3-indolemethanol hydrate, (33) 3-indole ethanol (tryptophol), (34) indole-3-carboxaldehyde, (35) 3-indolylacetate (3-acetoxyindole), (36) indole-3-acetamide, (37) indole-3-carboxylic acid, (38) indole-3-acetic acid, (39) 3-Indole propionic acid, (40) 3-indole acrylic acid, (41) 3-indole glyoxylic acid, (42) indole-3-pyruvic acid, (43) D,L-3-indolelactic acid, (44) 3-indole butyric acid, (45) N-acetyl-L-tryptophanamide,(46) N-(3-indolylacetyl)-L-alanine, (47) N-(3-indolyl acetyl)-L-valine, (48) N-(3-indolyl acetyl)-L-isoleucine, (49) N-(3-indolyl acetyl)-L-leucine, (50) N-(3-indolyl acetyl)-D,L-aspartic acid, (51) N-(3-indolyl acetyl)-L-phenylalanine, (52) 4-hydroxyindole (4-Indolol), (53) indole-4-carboxylic acid, (54) 4-indolyl acetate, (55) 4-methyl indole, (56) 5-hydroxy indole (5-indolol), (57) 5-hydroxy indole-3-acetic acid, (58) 5-hydroxy-2-indole carboxylic acid, (59) N-acetyl-5-hydroxytryptamine, (60) indole-5-carboxylic acid, (61) 5-methyl indole, (62) 5-methoxy indole, (63) indole-2-carboxylic acid, (64) D,L-indolene-2-carboxylic acid, (65) indole-2,3-dione (isatin), (66) 2-methyl indole, (67) 2,3,3-trimethyl indolenine, (68) tryptamine hydrochloride, (69) 5-methyl tryptamine hydrochloride, (70) serotonin hydrochloride hemihydrate (5-hydroxy tryptamine hydrochloride hemihydrate), (71) norharman hydrochloride monohydrate, (72) harmane hydrochloride monohydrate, (73) harmine hydrochloride hydrate, (74) harmaline hydrochloride dihydrate, (75) harmol hydrochloride dihydrate, (76) harmalol hydrochloride dihydrate, (77) 3,6-diamino acridine hydrochloride, (78) S-(3-indolyl) isothiuronium iodide, (79) yohimbine hydrochloride, and the like.

(H) pyrazoles and pyrazole derivatives, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻_{,} CH₃C₆H₄SO₃⁻, SO₃²⁻, BrO₃⁻, lO₃⁻, BrO₃⁻, or the like, as well as mixtures thereof.

Examples of suitable pyrazole compounds include (1) pyrazole, (2) 3-amino pyrazole, (3) 5-amino-1-ethylpyrazole, (4) 3-amino-4-carbethoxypyrazole, (5) 3-amino-5-methylpyrazole, (6) 3-amino-5-phenylpyrazole, (7) ethyl 4-pyrazole carboxylate, (8) diethyl 3,5-pyrazolecarboxylate, (9) 1,1'-(1-ethylpropylidene)bis 1H-pyrazole, (10) 4-bromopyrazole, (11) 4-bromo-3-methyl pyrazole, (12) 3,5-dimethyl pyrazole, (13) 4-bromo-3,5-dimethyl pyrazole, (14) 3,5-dimethyl pyrazole-1-carboxamide, (15) 3,5-dimethylpyrazole-1-methanol, (16) 3-methyl-1-vinylpyrazole, (17) 4-benzoyl-3-methyl-1-phenyl-2-pyrazolin-5-one, (18) 1-nitropyrazole, (19) 4-pyrazole carboxylic acid, (20) 3,5-pyrazole dicarboxylic acid monohydrate, (21) 3-amino-5-hydroxypyrazole, (22) 3-amino-4-pyrazole carbonitrile, (23) 3-amino-4-pyrzaolecarboxylic acid, (24) 4-methyl pyrazole hydrochloride, (25) 3,4-diamino-5-hydroxy pyrazole sulfate, (26) (3,5-dimethyl pyrazole-1-carboxamidine nitrate), (27) 3-amino-4-pyrazole carboxamide hemisulfate, (28) acid salt of 6-amino indazole hydrochloride, (29) 4-hydroxypyrazolo [3,4-d] pyrimidine, (30) 4-mercapto-1H-pyrazolo-[3,4-d]-pyrimidine, (31) indazole, (32) 5-aminoindazole, (33) 6-aminoindazole, (34) 3-indazolinone, (35) N'-(6-indazolyl) sulfanilamide, (36) 4,5-dihydro-3-(4-pyridinyl)-2H-benz[g] indazole methane sulfonate, and the like;

(I) Imidazoles and imidazole derivatives, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable imidazole compounds include (1) imidazole, (2) 4-methylimidazole, (3) 2-ethylimidazole, (4) 2-propylimidazole, (5) 1-butylimidazole, (6) 2-undecylimidazole,(7) histamine, (8) 1-(3-aminopropyl) imidazole, (9) 1-acetylimidazole, (10) 2-methyl-1-vinylimidazole,(11) 2-ethyl-4-methylimidazole, (12) 1-benzyl-2-methylimidazole, (13) 1-methylbenzimidazole, (14) 1-ethyl-3-methyl-1,H-imidazolinium chloride, (15) 2-(aminomethyl) benzimidazole dihydrochloride hydrate, (16) 2,6-diamino-8-purinol hemisulfate monohydrate, (17) purin-6-yl-trimethyl ammonium chloride, (18) 4-methyl-5-imidazole methanol hydrochloride, (19) N,N'-bis[3-(4,5-dihydro-1H-imidazol-2-yl)phenyl]urea dipropanoate, (20) 1-(p-tosyl)-3,4,4-trimethyl-2-imidazolinium iodide, (21) 1-ethyl-3-methyl-1H-imidazolinium chloride, (22) 2-amino imidazole sulfate, (23) 4-amino-5-imidazole carboxamide hydrochloride, (24) 2-hydrazino-2-imidazoline hydrobromide, (25) imidazole hydrochloride, (26) 4-imidazole acetic acid hydrochloride, (27) 2-benzyl-2-imidazoline hydrochloride, (28) propyl-1-(1-phenyl ethyl imidazole-5-carboxylate hydrochloride, (29) 2,6-diamino purine sulfate hydrate, (30) 1-tallow amido ethyl-3-methyl-2-heptadecyl imidazolinium methyl sulfate, (31) isostearyl ethyl imidonium ethyl sulfate, (32) methyl (1) tallow amido ethyl-2-tallow imidazolinium methyl sulfate, (33) isostearyl benzyl imidonium chloride, (34) methyl (1) hydrogenated tallow amido ethyl (2) hydrogenated tallow imidazolinium methyl sulfate, (35) 1-methyl-1-oleyl amido ethyl-2-oleyl-imidazolinium methyl sulfate, (36) cocohydroxyethyl polyethyleneglycol imidazolinium chloride phosphate, (37) 1-methyl uric acid, (38) guanine, (39) guanosine hydrate, (40) xanthine, (41) 1-methylxanthine, (42) 3-methyl xanthine, (43) 3-isobutyl-1-methyl xanthine, (44) hypoxanthine, (45) xanthosine dihydrate, (46) 6-thioxanthene, (47) purine, (48) 6-amino purine (adenine), (49) 6-methoxy purine hemihydrate, (50) 6-mercaptopurine monohydrate, (51) 2-amino-6-chloropurine, (52) 2-amino-6,8-dihydroxy purine, (53) theophylline (3,7 dihydro-1,3-dimethyl-1H-purine-2,6-dione), (54) kinetin (6-furfuryl amino purine), (55) 1-methyl adenine, (56) 3-methyl adenine, (57) (-)-adenosine, (58) (-)-inosine, (59) 6-mercaptopurine riboside, (60) 6-amino purine hydrochloride hemihydrate, (61) 6-amino purine sulfate, (62) 2,6-diamino-8-purinol hemisulfate monohydrate, (63) benzimidazole, (64) 2-aminobenzimidazole, (65) 2-amino-5,6-dimethlybenzimidazole, (66) 5-benzimidazole carboxylic acid, (67) 2,4,5-trimethyl benzimidazole, (68) 2-guanidinobenzimidazole, (69) 2-hydroxybenzimidazole, (70) 4-(2-keto-1-benzimidazolinyl) piperidine, (71) 2-imidazolidine thione, (72) 2-imidazolidone, (73) hydantoin, (74) 1-methyl hydantoin, (75) creatinine, (76) 2-thiohydrantoin, (77) 5-hydantoin acetic acid, (78) 5-ureidohydantoin (allantoin), (79) 5,5-dimethyl hydantoin, (80) 2-imidazolidone-4-carboxylic acid, and the like;

(J) pyridines and pyridine derivatives, including those of the general formula wherein R₁, R₂, R₃, R₄, and R₅ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, and R₅ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable pyridine compounds include (1) N,N-bis (2-hydroxyethyl) isonicotinamide, (2) 1,2-bis(4-pyridyl) ethylene, (3) 2-(2-piperidinoethyl) pyridine, (4) 1,2-bis (4-pyridyl)ethane, (5) 4,4'-trimethylene pyridine, (6) aldrithiol-2, (7) aldrithiol-4, (8) 1,3-bis (3-pyridylmethyl)-2-thiourea, (9) 2,2':6',2"-terpyridine, (10) 2-[N,N-bis(triflouromethylsulfonyl)amino]pyridine, (11) 2,3-pyridine dicarboxylic acid, (12) 2,4-pyridine dicarboxylic acid monohydrate, (13) 2,5-pyridine dicarboxylic acid, (14) 2,6-pyridine dicarboxylic acid, (15) 3,4-pyridine dicarboxylic acid, (16) 3,5-pyridine dicarboxylic acid, (17) 2,6-pyridine dicarboxaldehyde, (18) 3,4-pyridine carboxamide, (19) 3,4-pyridine carboximide, (20) 2,3-pyridine carboxylic anhydride, (21) 3,4-pyridine carboxylic anhydride, (22) 2,6-pyridine methanol, (23) 2-pyridine ethane sulfonic acid, (24) 4-pyridine ethane sulfonic acid, (25) 3-pyridine sulfonic acid, (26) pyridoxic acid, (27) trans-3-(3-pyridyl) acrylic acid, (28) 2-pyridyl hydroxymethane sulfonic acid, (29) 3-pyridyl hydroxymethane sulfonic acid, (30) 6-methyl-2,3-pyridine dicarboxylic acid, (31) isonicotinic acid, (32) pyridine hydrobromide, (33) pyridine hydrochloride, (34) 2-(chloromethyl) pyridine hydrochloride, (35) 2-pyridylacetic acid hydrochloride, (36) nicotinoyl chloride hydrochloride, (37) 2-hydrazinopyridine dihydrochloride, (38) 2-(2-methyl aminoethyl) pyridine dihydrochloride, (39) 1-methyl-1,2,3,6-tetrahydropyridine hydrochloride, (40) 2,6-dihydroxypyridine hydrochloride, (41) 3-hydroxy-2(hydroxymethyl) pyridine hydrochloride, (42) pyridoxine hydrochloride, (43) pyridoxal hydrochloride, (44) pyridoxal 5-phosphate monohydrate, (45) 3-amino-2,6-dimethoxy pyridine hydrochloride, (46) pyridoxamine dihydrochloride monohydrate, (47) iproniazid phosphate (isonicotinic acid 2-isopropyl hydrazide phosphate), (48) tripelennamine hydrochloride, (49) pyridinium bromide perbromide, (50) pyridinium 3-nitrobenzenesulfonate, (51) 1-ethyl-3-hydroxy pyridinium bromide, (52) 1-ethyl-4-(methoxy carbonyl) pyridinium iodide, (53) 1-heptyl-4-(4-pyridyl) pyridinium bromide, (54) 1-dodecyl pyridinium chloride, (55) 1-hexadecyl pyridinium chloride monohydrate, (56) 1-hexadecyl pyridinium bromide monohydrate, (57) 1-(carboxymethyl) pyridinium chloride, (58) 1-(carboxymethyl) pyridinium chloride hydrazide, (59) 1-(3-nitrobenzyloxymethyl) pyridinium chloride, (60) 1-(3-sulfopropyl) pyridinium hydroxide, (61) N-(lauroyl colamino formyl methyl) pyridinium chloride, (62) N-(stearoyl colamine formyl methyl) pyridinium chloride, (63) 2-chloro-1-methyl pyridinium iodide, (64) 2-pyridine aldoxime-1-methyl methane sulfonate, (65) 2-pyridine aldoxime-1-methyl chloride, (66) 2-[4-(dimethyl amino) styryl]1-ethylpyridinium iodide, (67) 1-benzyl-3-hydroxy pyridinium chloride, (68) 1,4 dimethyl pyridinium iodide, (69) 1-ethyl-4-phenyl pyridinium iodide, (70) 4-phenyl-1-propyl pyridinium iodide, (71) 1-docosyl-4-(4 hydroxystyryl) pyridinium bromide, (72) 1,1'-dimethyl-4-4'-bipyridinium dichloride, (73) 1,1'-diethyl-4-4'-bipyridinium dibromide, (74) 1,1'-dibenzyl-4,4'-bipyridinium dichloride, (75) 1,1'-diheptyl-4,4'-bipyridinium dibromide, (76) 1,7-phenanthroline, (77) 1,10-phenanthroline, (78) 5-chloro-1,10-phenanthroline, (79) 4,5-dihydro-3-(4-pyridinyl)-2H-benz[g] indazole methane sulfonate, and the like;

(K) quinolines and quinoline derivatives, and isoquinolines and isoquinoline derivatives, including those of the general formulae wherein R₁, R₂, R₃, R₄, R₅, R₆, R₇, R₈, R₉, R₁₀, R₁₁, R₁₂, R₁₃, and R₁₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, and R₁₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable quinoline and isoquinoline compounds include (1) 1,2,3,4-tetrahydro quinoline, (2) 6-ethoxy-1,2,3,4-tetrahydro-2,2,4-trimethyl quinoline, (3) 2-cyanoquinoline, cyanoquinoline, (4) 1-cyanoisoquinoline, (5) 3-cyanoisoquinoline, (6) 3-amino quinoline, (7) (8) 7,8-benzoquinoline, (9) 8-hydroxy quinoline, (10) 8-hydroxyquinoline, aluminium salt, (11) 8-hydroxyquinaldine, (12) 3,4,5,6,7,8-hexahydro 2 (1H)-quinolinone, (13) julolidine, (14) quinoxaline, (15) ethyl-2-quinoxalinecarboxylate, (16) quinoline, (17) 2-hydroxyquinoline, (18) 4-hydroxy quinoline, (19) 5-hydroxy quinoline, (20) 5-amino quinoline, (21) 6-amino quinoline, (22) 2-quinoline carboxylic acid, (23) 3-quinoline carboxylic acid, (24) 4-quinoline carboxylic acid, (25) 4-quinoline carboxaldehyde, (26) 2-quinoline thiol, (27) 2,4-quinoline diol, ((28) quinaldine, (29) 4-aminoquinaldine, (30) 2,6-dimethyl quinoline, (31) 2,7-dimethyl quinoline, (32) 4-methoxy-2-quinoline carboxylic acid, (33) methyl-2-phenyl-4-quinoline carboxylate, (34) 2-(N-butyl carbamoyl)-1,2,3,4-tetrahydro-isoquinoline, (35) 1-hydroxyisoquinoline, (36) 1-isoquinoline carboxylic acid, (37) 3-isoquinoline carboxylic acid, (38) 1,5-isoquinoline diol, (39) 8-hydroxyquinoline hemisulfate hemihydrate, (40) 5-amino-8-hydroxy quinoline dihydrochloride, (41) 2-(chloromethyl) quinoline monohydrochloride, (42) 8-hydroxyquinoline-5-sulfonic acid monohydrate, (43) 8-ethoxy-5-quinoline sulfonic acid sodium salt hydrate, (44) 1,2,3,4-tetrahydroisoquinoline hydrochloride, (45) 1,2,3,4-tetrahydro-3-isoquinoline carboxylic acid hydrochloride, (46) 6,7-dimethoxy-1,2,3,4-tetrahydro isoquinoline hydrochloride, (47) 1-methyl-6,7-dihydroxy-1,2,3,4-tetrahydro isoquinoline hydrobromide, (48) primaquine diphosphate [8-(4-amino-1-methyl butyl amino)-6-methoxy quinoline diphosphate], (49) pentaquine phosphate, (50) dibucaine hydrochloride [2-butoxy-N-(2-diethyl amino ethyl)-4-quinoline carboxamide hydrochloride], (51) 9-aminoacridine hydrochloride hemihydrate, (52) 3, 6-diamino acridine hemisulfate, (53) 2-quinoline thiol hydrochloride, (54) (-) sparteine sulfate pentahydrate, (55) papaverine hydrochloride, (56) (+)-emetine dihydrochloride hydrate, (57) 1,10-phenanthroline monohydrochloride monohydrate, (58) neocuproine hydrochloride trihydrate, and the like;

(L) pyrimidines and pyrimidine derivatives, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, IO₃⁻, BrO₃⁻, or the like, as well as mixtures thereof.

Examples of suitable pyrimidines include (1) pyrimidine, (2) 2 chloropyrimidine, (3) 4-phenylpyrimidine, (4) 5-bromopyrimidine, (5) 2,4-dichloropyrimidine, (6) 4,6-dichloropyrimidine, (7) 2,4-dichloro-6-methylpyrimidine, (8) 6-chloro-2,4-dimethoxypyrimidine, (9) 2-amino-4,6-dimethoxypyrimidine, (10) 2,4,6-trichloropyrimidine, (11) 2,4,5,6-tetrachloropyrimidine, (12) 1,3,4,6,7,8-hexahydro-1-methyl-2H-pyrimido [1,2-a] pyrimidine, (13) 1,3,4,6,7,8-hexahydro-2H-pyrimido [1,2-a] pyrimidine, (14) hexetidine, (15) tert-butyl S-(4,6-dimethylpyrimidin-2-yl) thiocarbonate, (16) 4-methoxybenzyl-S(4,6-dimethylpyrimidin-2-yl) thiocarbonate, (17) 2-amino pyrimidine, (18) 2-amino-4-methyl pyrimidine, (19) 2-amino-5-nitropyrimidine, (20) 2-amino-5-bromopyrimidine, (21) 2-amino-4-chloro-6-methyl pyrimidine, (22) 2-amino-4,6-dimethyl pyrimidine, (23) 2-amino-4-hydroxy-6-methyl pyrimidine, (24) 2-amino-4,6-dichloropyrimidine, (25) 2-amino-5-bromo-6-methyl-4-pyrimidinol, (26) 4-aminopyrimidine, (27) 4,5-diamino pyrimidine, (28) 4-amino-2,6-dimethyl pyrimidine, (29) 2,4-diamino-6-hydroxypyrimidine, (30) 2,6-diamino-4-chloro pyrimidine, (31) 4,6-diamino-2-mercaptopyrimidine hemihydrate, (32) 2,4,6-triamino pyrimidine, (33) 5-nitroso-2,4,6-triamino pyrimidine, (34) 4,6-dihydroxy pyrimidine, (35) 4,6-dihydroxy-2-amino pyrimidine, (36) 4,6-dihydroxy-2-methyl pyrimidine, (37) 4,6-dihydroxy-5-nitropyrimidine, (38) 2,4-dihydroxy-5-methyl pyrimidine, (39) 2,4-dihydroxy-6-methyl pyrimidine, (40) 2,4-dihydroxy-5,6-dimethyl pyrimidine, (41) 2,6-dihydroxy pyrimidine-5-carboxylic acid hydrate, (42) 2,6-dihydroxy-4-amino pyrimidine, (43) 2,4,5-trihydroxy pyrimidine, (44) 2-thiouracil [4-hydroxy-2-mercaptopyrimidine], (45) 6-amino-5-nitroso-2-thiouracil, (46) folic acid dihydrate, (47) folinic acid, calcium salt hydrate, (48) 2-hydroxypyrimidine hydrochloride, (49) 2-hydroxy-4-methyl pyrimidine hydrochloride, (50) 4,6-dimethyl-2-hydroxypyrimidine hydrochloride, (51) 2-mercapto-4-methyl pyrimidine hydrochloride, (52) 4,6-diamino pyrimidine hemisulfate monohydrate, (53) 4,5,6-triamino pyrimidine sulfate hydrate, (54) 4,5-diamino-6-hydroxy pyrimidine sulfate, (55) 2,4-diamino-6-mercapto pyrimidine hemisulfate, (56) 2,4-diamino-6-hydroxy pyrimidine hemisulfate hydrate, (57) 6-hydroxy-2,4,5-triamino pyrimidine sulfate, (58) 5,6-diamino-2,4-dihydroxy pyrimidine sulfate, (59) N4-(2-amino-4-pyrimidinyl) sulfanilamide monohydrochloride, (60) 2,4,5,6-tetraamino pyrimidine sulfate, (61) pyrimidine diones, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃-, SO₃²⁻, BrO₃⁻, lO₃⁻, ClO₃⁻, or the like, as well as mixtures thereof, such as (a) 2,4 (1H,3H)-pyrimidine dione (uracil), (b) 5-amino uracil, (c) 5-nitrouracil, (d) 5-iodouracil, (e) 5-(hydroxymethyl) uracil hydrate, (f) 5,6-dihydrouracil, (g) 6-amino-1-methyl uracil, (h) 5,6-diamino-1,3-dimethyl uracil hydrate, (i) uridine, (j) 5-methyl uridine, (k) 5-iodouridine, (I) thimidine, and the like; (62) thiouracils, such as (a) 5-methyl-2-thiouracil, (b) 4-thiouridine, (c) 2-thiocytidine dihydrate, and the like; (63) orotic acid compounds, such as (a) orotic acid monohydrate, (b) L-hydroorotic acid, (c) 5-aminoorotic acid, (d) methylorotate (orotic acid methyl ester), and the like; (64) pyrimidine trione compounds, such as (a) barbituric acid, (b) 5-nitrobarbituric acid trihydrate, (c) violuric acid monohydrate, (d) alloxan monohydrate [2,4,5,6-(1H,3H)-pyrimidine-tetrone], (65) 4,5,6-triamino-2(1H)-pyrimidinethione sulfate, (66) (-)-cyclocytidine hydrochloride, (67) cytosine arabinoside hydrochloride, and the like;

(M) pyradizines and pyridazine derivatives, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable pyridazines include (1) pyridazine, (2) phthalazine, (3) 4,5-dihydro-6-methyl-3(2H)-pyridazinone monohydrate, (4) 3,6-dichloropyridazine, (5) 3,4,5-trichloropyridazine, (6) 3,6-dichloro-4-methylpyridazine, (7) 3-chloro-6-methoxypyridazine, and the like;

(N) pyrazines and pyrazine derivatives, including those of the general formula wherein R₁, R₂, R₃, and R₄ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, and R₄ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable pyrazines include (1) pyrazine, (2) acetylpyrazine, (3) aminopyrazine, (4) 2,6-dichloropyrazine, (5) 2,3,5-trimethylpyrazine, (6) tetramethylpyrazine, (7) 5-methyl-2-pyrazine carboxylic acid, (8) pyrazine amide, (9) 2,3-pyrazine dicarboxamide, (10) 4-pyridazine carboxylic acid, (11) 2,3-pyrazine dicarboxylic acid, (12) lumazine monohydrate, (13) xanthopterin monohydrate, (14) 2-quinoxazoline carboxylic acid, (15) 2-quinoxalinol, (16) 2,3-dihydroxy quinoxaline, (17) phenazine methosulfate, and the like;

(O) lactams and lactam derivatives, and thiolactams and thiolactam derivatives, including those of the general formulae wherein R₁ can be selected from (but is not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, and wherein the curved portion of the structure represents a hydrocarbon chain or a substituted hydrocarbon chain, preferably of from about 2 to about 10 carbon atoms, wherein two or more substituents can be joined together to form a ring, and wherein the substituents on the substituted alkyl groups, substituted aryl groups, substituted arylalkyl groups, and substituted hydrocarbon chain can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable lactams and thiolactams include (1) 2-azetidinone (β-propiolactam), propiolactam), (2) 2-pyrrolidinone, (3) pyrrolidone hydrotribromide, (4) δ-valerolactam, (5) ε-caprolactam, (6) amino-ε-caprolactam, (7) N-methyl caprolactam, (8) 2-azacyclooctanone, (9) 2-azacyclononanone, (10) ω-thiocaprolactam, (11) N-vinylcaprolactam, (12) (±)-2-azabicyclo[2.2.1]hept-5-en-3-one, and the like;

(P) imides and imide derivatives, including those of the general formula wherein R₁ can be selected from (but is not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, and wherein the curved portion of the structure represents a hydrocarbon chain or a substituted hydrocarbon chain, preferably of from about 1 to about 20 carbon atoms, wherein two or more substituents can be joined together to form a ring, and wherein the substituents on the substituted alkyl groups, substituted aryl groups, substituted arylalkyl groups, and substituted hydrocarbon chain can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable imide compounds include (1) maleimide, (2) N-ethylmaleimide, (3) N-butylmaleimide, (4) N-cyclohexylmaleimide, (5) N-phenylmaleimide, (6) N-benzylmaleimide, (7) N-hydroxymaleimide, (8) succinimide, (9) N-methylsuccinimide, (10) (S)-(-)-2-hydroxy-N-methylsuccinimide, (11) N-hydroxysuccinimide, (12) succinimidyl 2,2,2-trichloroethyl carbonate, (13) 2-dodecyl-N-(2,2,6,6-tetramethyl-4-ppiperidinyl) succinimide, (14) 2-dodecyl-N-(1,2,2,6,6-pentamethyl-4-piperdinyl) succinimide, (15) N-(1-acetyl-2,2,6,6-tetramethyl-4-piperidinyl)-2-dodecyl succinimide, (16) α-methyl-α-propylsuccinimide, (17) α-methyl-α-phenylsuccinimide, (18) N-vinylphthalimide, (19) N-ethylphthalimide, (20) N-(trimethylsilylmethyl)phthalimide, (21) N-(2-bromoethyl)phthalimide, (22) N-(3-bromopropyl)phthalimide, (23) N-(4-bromobutyl)phthalimide, (24) phthalimidoacetaldehyde diethyl acetal, (25) diethyl (phthalimidomethyl)phosphonate, (26) N-benzylphthalimide, (27) phthalimide, DBU (1,8-diazabicyclo [5.4.0]undec-7-ene) salt, (28) phthalimide, DBN (1,5-diazabicyclo [4.3.0]non-5-ene), and the like;

II. Oxa-aza-cyclic compounds, including (A) oxazoles and oxazole derivatives, and isoxazoles and isoxazole derivatives, including those of the general formulae wherein R₁, R₂, R₃, R₄, R₅, R₆, R₇, R₈, R₉, R₁₀, R₁₁, R₁₂, R₁₃, R₁₄, and R₁₅ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, R₁₄, and R₁₅ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable oxazole and isoxazole compounds include (1) 3-amino-5-methyl isoxazole, (2) 5-amino-3-methyl isoxazole, (3) 3,5-dimethyl-4-nitroisoxazole, (4) 1,2-benzisoxazole, (5) 2,1-benzisoxazole (Anthranil), (6) cycloserine [4-amino-3-isoxazolidinone], (7) 4-benzyl-2-methyl-2-oxazoline, (8) 2-methyl-5-phenyl-2-oxazoline-4-methanol, (9) benzoxazole, (10) 2-methylbenzoxazole, (11) 2-chlorobenzoxazole, (12) 2-chloro-3-ethylbenzeneoxazolium tetrafluoroborate, (13) 2-oxazolidone, (14) 3-methyl-2-oxazolidinone, (15) 5-chloromethyl-2-oxazolidinone, (16) 4-isopropyl-2-oxazolidinone, (17) 3-acetyl-2-oxazolidinone, (18) 5,5-dimethyl oxazolidine-2,4-dione, (19) 3-ethyl-2-thioxo-4-oxazolidinone, (20) 4-methyl-5-phenyl-2-oxazolidinone, (21) 4-benzyl-2-oxazolidinone, (22) 2-benzoisoxazolinone, (23) muscimol hydrate [5-(aminomethyl)-3-isoxazolol hydrate], (24) 5-methyl-3-phenyl isoxazole-4-carboxylic acid, (25) 2-methyl-5-phenyl-2-oxazoline-4-methanol, (26) sulfamethoxazole [4-amino-N-(5-methyl-3-isoxazolyl) benzene sulfonamide], (27) sulfisoxazole [4-amino-N-(3,4-dimethyl-5-isoxazolyl) benzene sulfonamide], (28) N'-(4,5-dimethyloxazol-2-yl) sulfanilamide, (29) cycloserine [4-amino-3-isoxazolidinone], (30) chlorzoxazone [5-chloro-2-benzoxazolone], (31) 3,3'-dimethyl oxacarbocyanine iodide, (32) 2-ethyl-5-phenyl isoxazolium-3'-sulfonate, (33) 2-chloro-3-ethylbenzoxazolium tetrafluoroborate, (34) 2-tert-butyl-5-methyl isoxazolium perchlorate, (35) 5-phenyl-2-(4-pyridyl) oxazole hydrochloride hydrate, (36) 5-phenyl-2-(4-pyridyl) oxazole methyl tosylate salt, and the like;

(B) morpholines and morpholine derivatives, including those of the general formula wherein R₁, R₂, R₃, R₄, R₅, R₆, R₇, R₈, and R₉ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, and R₉ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable morpholines include (1) 4-aminomorpholine, (2) 4-morpholine carbonitrile, (3) 4-morpholine propionitrile, (4) 4-formyl morpholine, (5) 4-acetylmorpholine, (6) 4-(2-hydroxyethyl) morpholine, (7) 3-morpholino-1,2-propane diol, (8) 4-(3-amino propyl) morpholine, (9) 1-morpholino-1-cyclopentene, (10) 1-morpholino-1-cyclohexene, (11) 1-morpholino-1-cycloheptene, (12) 4-phenyl morpholine, (13) 4-morpholinoaniline, (14) 2,2,2-tribromoethyl phosphoromorpholino chloridate, (15) 1-(morpholino carbonyl methyl) piperazine, (16) 1,3-dimorpholine-2-nitropropane, (17) hemicholinium-3, (18) hemicholinium-15, (19) 2-methoxy-4-morpholinobenzene diazoniumchloride, zinc chloride, (20) fomocaine, (21) 4-morpholinobenzophenone, (22) 4,4'-ethylene-bis (2,6-morpholinedione), (23) N,N'-dicylcohexyl-4-morpholine carboxamidine, (24) 1-cyclohexyl-3-(2-morpholino ethyl)-2-thiourea, (25) 4-morpholinoacetophenone, (26) 4-(2-chloroethyl) morpholine hydrochloride, (27) 4-morpholine ethane sulfonic acid, (28) 4-morpholine propane sulfonic acid, (29) β-hydroxy morpholine propane sulfonic acid, (30) [N-(aminoiminomethyl)-4-morpholine carboximidamide] hydrochloride, (31) 4-morpholine carbodithioic acid compound with morpholine, (32) 2,5-dimethyl-4-(morpholinomethyl) phenol hydrochloride monohydrate, (33) 1-cyclohexyl-3-(2-morpholinoethyl) carbodiimide metho-p-toluene sulfonate, (34) hemicholinium-3[2,2'-(4,4'-biphenylene) bis(2-hydroxy-4,4-dimethyl morpholinium bromide), (35) hemicholinium-15[4,4-dimethyl-2-hydroxy-2-phenyl morpholinium bromide], and the like; (C) cyclic aza-ethers and diazaethers, such as (1) 1-aza-12-crown-4, (2) 1-aza-15-crown-5, (3) 1-aza-18-crown-6, (4) 1,4,10-trioxa-7,13-diazacyclopentadecane, (5) 1,4,10,13-tetraoxa-7,16-diazacyclooctadecane, (6) N,N'-dibenzyl-1,4,10,13-tetraoxa-7,16-diazacyclooctadecane, (7) 4,7,13,18-tetraoxa-1,10-diazabicyclo [8.5.5] eicosane, (8) 4,7,13,16,21-pentaoxa-1,10-diazabicyclo [8.5.5] tricosane, (9) 4,7,13,16,21,24-hexaoxa-1,10-diazabicyclo [8.8.8] hexacosane, (10) 5,6-benzo-4,17,13,16,21,24-hexaoxa-1,10-diazabicyclo[8.8.8] hexacosane, and the like;

III. Oxacyclic compounds, including (A) cyclic compounds wherein the ring contains one oxygen atom, such as (1) lactones and lactone derivatives, including those of the general formula wherein the curved portion of the structure represents a hydrocarbon chain or a substituted hydrocarbon chain, preferably of from about 2 to about 20 carbon atoms, wherein two or more substituents can be joined together to form a ring, and wherein the substituents on the hydrocarbon chain can be (but are not limited to) alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of lactone compounds include (a) γ-butyrolactone, (b) γ-valerolactone, (c) γ-caprolactone, (d) γ-octanoic lactone, (e) γ-nonanoic lactone, (f) γ-decanolactone, (g) undecanoic γ-lactone, (h) γ-phenyl-γ-butyrolactone, (i) (±)-α-carbethoxy-γ-phenyl-butyrolactone, (j) 2-coumaranone, (k) (±)-β,β-dimethyl-γ-(hydroxymethyl)-γ-butyrolactone, (I) (S)-(+)-γ-ethoxy carbonyl-γ-butyrolactone, (m) (S)-(-)-5-(hydroxymethyl)-2(5H)-furanone, (n) dihydro-4,4-dimethyl-2,3-furandione, (o) 2,5-dimethyl-4-hydroxy-3(2H)-furanone, (p) (±)-mevalonic (β-hydroxy β-methyl-δ-valero) lactone, (q) (±)-δ-decanolactone, (r) (±)-undecanoic δ-lactone, (s) (±)-δ-dodecanolactone, (t) undecanoic ω-lactone, (u) oxacyclotridecan-2-one, (v) ω-pentadecalactone, (w) hydrindantin (2,2'-dihydroxy-2,2'-biindan-1,1'3,3'-tetrone, (x) hydrindantin dihydrate, (y) 2-oxepanone, and the like;
(2) pyrans and pyran derivatives, including those of the general formulae wherein R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, and R₂₈ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, and R₂₈ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of pyran compounds include (a) 4H-pyran-2-one, (b) methylcoumalate (methyl-2-oxo-2H-pyran-5-carboxylate, (c) methyl 2-oxo-2H-pyran-3-carboxylate, (d) 4,6-dimethyl-α-pyrone, (e) 4-methoxy-6-methyl-2H-pyran-2-one, (f) 2-oxo-6-pentyl-2H-pyran-3-carboxylic acid, (g) methylisodehydracetate, (h) ethylisodehydracetate, (i) 5,6-dihydro-2H-pyran-2-one, (j) 3,6-dihydro-4,6,6-trimethyl-2H-pyran-2-one, (k) 3,4-dihydro-6-methyl-2H-pyran-2-one, (I) 3-acetyl coumarin, (m) 6-methyl coumarin, (n) 7-ethoxy coumarin, (o) ethyl-3-coumarin carboxylate, (p) 7-diethylamino-4-methyl coumarin, (q) dihydro coumarin, (r) 3-bromo-2-coumaranone, (s) patulin (4-hydroxy-4H-furo[3.2.c]pyran-2(6H)-one), (t) 4H-pyran-4-one, (u) 2-ethyl-3-hydroxy-4H-pyran-4-one, (v) butopyronoxyl(butyl 3,4-dihydro-2,2-dimethyl-4-oxo-2H-pyran-6-carboxylate, (w) dehydroacetic acid, (x) 4-chromone (1-benzylpyran-4(4H)-one), (y) 4-chromanone, (z) 4-chromanol, (aa) 6,7-dimethoxy-2,2-dimethyl-4-chromanone, (bb) 3-isochromanone, (cc) 6,7-dimethoxy-3-isochromanone, (dd) 6-ethyl-4-oxo-4H-1-benzopyran-3-carbonitrile, (ee) 6-ethyl-4-oxo-4H-1-benzopyran-3-carboxaldehyde, (ff) 6-isopropyl-4-oxo-4H-1-benzopyran-3-carbonitrile, (gg) 6-isopropyl-4-oxo-4H-1-benzopyran-3-carboxaldehyde, and the like;
(3) cyclic anhydrides and anhydride derivatives, including those of the general formulae wherein the curved portion of the structure represents a hydrocarbon chain or a substituted hydrocarbon chain, preferably of from about 1 to about 20 carbon atoms, wherein two or more substituents can be joined together to form a ring, and wherein the substituents on the hydrocarbon chain can be (but are not limited to) alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃-, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of cyclic anhydrides include (a) maleic anhydride, (b) bromomaleic anhydride, (c) citraconic anhydride, (d) 2,3-dimethylmaleic anhydride, (e) dichloromaleic anhydride, (f) cis-aconitic anhydride, (g) itaconic anhydride, (h) methylsuccinic anhydride, (i) S-acetylmercaptosuccinic anhydride, (j) 2,2-dimethylsuccinic anhydride, (k) phenylsuccinic anhydride, (l) (±)-2-octen-1-ylsuccinic anhydride, (m) 2-dodecen-1-ylsuccinic anhydride, (n) 2-octadecen-1-ylsuccinic anhydride, (o) 3-oxabicyclo [3.1.0] hexane-2,4-dione, (p) diglycolic anhydride, (q) glutaric anhydride, (r) 3-methylglutaric anhydride, (s) 2,2-dimethylglutaric anhydride, (t) 3,3-tetramethyleneglutaric anhydride, (u) 1-cyclopentene-1,2-dicarboxylic anhydride, (v) 3,4,5,6-tetrahydrophthalic anhydride, (w) cis-1,2-cyclohexanedicarboxylic anhydride, (x) (±)-hexahydro-4-methylphthalic anhydride, (y) methyl-5-norbornene-2,3-dicarboxylic anhydride, (z) 2,3-pyridinecarboxylic anhydride, (aa) 3,4-pyridinecarboxylic anhydride, and the like; (4) cyclic oxa-sulfur compounds and their derivatives, including (a) furfurylmercaptan, (b) S-furfurylthioacetate, (c) furfurylsulfide, (d) furfurylmethyldisulfide, (e) furfuryldisulfide, and the like;
(B) cyclic compounds wherein the ring contains at least two oxygen atoms, such as (1) dioxanes and dioxane derivatives, and trioxanes and trioxand derivatives, including those of the general formulae wherein R₁, R₂, R₃, R₄, R₅, R₆, R₇, and R₈ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, and R₈ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of suitable dioxanes and trioxanes include (a) glycolaldehyde dimer (2,5-dihydroxy-1,4-dioxane), (b) 6,7-dihydrocyclopenta-1,3-dioxin-5(4H)-one, (c) (2R,6R)-tert-butyl-6-methyl-1,3-dioxan-4-one, 6-methyl-1,3-dioxan-4-one, (d) 2,2-dimethyl-1,3-dioxane-4,6-dione, (e) (f) 2,2,6-trimethyl-4H-1,3-dioxin-4-one, (g) 2,2,5-trimethyl-1,3-dioxane-4,6-dione, (h) 5-bromo-2,2,5-trimethyl-1,3-dioxane-4,6-dione, (i) 1,3-dioxane-5,5-dimethanol, (j) 1,3,5-trioxane, and the like; (2) oxaspiros and oxaspiro derivatives, and ketals and ketal derivatives, including those of the general formulae wherein the curved portions of the structures represent a hydrocarbon chain or a substituted hydrocarbon chain, preferably of from 1 to about 20 carbon atoms, wherein two or more substituents can be joined together to form a ring, and wherein the substituents on the hydrocarbon chains can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of oxaspiros and ketals include (a) 1,6-dioxaspiro [4.4]nonane-2,7-dione, (b) 1,4-dioxaspiro [4.5]decan-2-one, (c) 1,7-dioxaspiro [5.5]undecane, (d) 2,4,8,10-tetraoxaspiro[5.5]undecane, (e) 3,9-divinyl-2,4,8-tetraoxaspiro[5.5]undecane, (f) 2,2-pentamethylene-1,3-dioxalane,(g) 2-phenyl-1,3-dioxalane, (h) 1,4-cyclohexanedione monoethylene ketal, (i) 1,4-cyclohexanedione bis(ethylene ketal), (j) 1,4-cyclohexanedione mono-2,2-dimethyl trimethylene ketal, and the like; (3) methylene dioxys and methylene dioxy derivatives, including those of the general formula wherein R₁, R₂, R₃, R₄, R₅, and R₆ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, and R₆ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, IO₃⁻, ClO₃⁻, or the like, as well as mixtures thereof.

Examples of suitable methylenedioxy compounds include (a) piperonal, (b) piperonyl acetate, (c) piperonyl alcohol, (d) piperonylnitrile, (e) piperonyl amine, (f) 6-nitropiperonal, (g) 6-nitropiperonyl alcohol, (h) 3',4'-(methylenedioxy)acetophenone, (i) 3,4-(methylenedioxy)aniline, (j) 2,3-(methylenedioxy)benzaldehyde, (k) 3,4-(methylenedioxy)phenylacetonitrile, (I) 3,4-(methylenedioxy)toluene, and the like;
(C) crown ethers, including (1) 1,4,7,10-tetraoxacyclododecane (12-crown-4), (2) 2-(hydroxyethyl)-12-crown-4, (3) 2-(aminoethyl)-12-crown-4, (4) benzo-12-crown-4, (5) 1,4,7,10,13-pentaoxacyclododecane (15-crown-5), (6) 2-(hydroxyethyl)-15-crown-5,(7) 2-(aminoethyl)-15-crown-5, (8) benzo-15-crown-5, (9) 4'-aminobenzo-15-crown-5, (10) 4'-formylbenzo-15-crown-5, (11) 4'-nitrobenzo-15-crown-5, (12) bis [(benzo-15-crown-5)-15-ylmethyl] pimelate, (13) 1,4,7,10,13,16-hexaoxacyclooctadecane (18-crown-6), (14) 2-(aminoethyl)-18 crown-6, (15) benzo-18 crown-6, (16) 4'-bromobenzo-18-crown-6, (17) dibenzo-18-crown-6 (2,3,11,12-dibenzo-1,4,7,10,13,16-hexaoxacyclooctadeca-2,11-diene), (18) di-tert-butyldibenzo-18-crown-6, (19) cis-dicyclohexane-18 crown-6 (2,3,11,12-dicyclohexano-1,4,7,10,13,16-hexaoxacyclooctadecane), (20) dibenzo-24-crown-8 [2,3,14,15-dibenzo,1,4,7,10,13,16,19,22-octaoxacyclotetracosa 2,14-diene], (21) dicyclohexano-24-crown-8, (22) dibenzo-30-crown-10,[2,3,17,18-dibenzo-1,4,7,10,13,16,19,22,25,28-decaoxacyclotriaconta-2,17-diene], and the like;

III. Cyclic hydrocarbons (wherein the compound contains at least one ring with only carbon atoms, although other rings present in the compound may contain atoms other than carbon and substituents may be present on the ring(s)), including (A) norbornanes and norbornane derivatives, and norbornenes and norbornene derivatives, including those of the general formulae wherein R₁, R₂, R₃, R₄, R₅, R₆, R₇, R₈, R₉, R₁₀, R₁₁, and R₁₂ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, and R₁₂ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, I⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, IO₃⁻, ClO₃⁻, or the like, as well as mixtures thereof.

Examples of norbornanes and norbornenes include (1) norbornane, (Aldrich N3,200-8), (2) 2-norbornane carbonitrile, (3) 2-norbornane methanol, (4) 3-methyl-2-norbornane methanol, (5) camphene, (6) fenchyl alcohol, (7) thiocamphor, (8) norbornene, (9) 5-norbornene-2-carbonitrile, (10) 5-norbornene-2-carboxaldehyde, (11) 5-norbornene-2-methanol, (12) 5-norbornene-2,2-dimethanol, (13) 5-norbornene-2-benzoyl, (14) 2-norbornanone (norcamphor), (15) 3-chloro-2-norbornanone, (16) fenchone (1,3,3-trimethyl-2-norbornanone, (17) (+)-3-(trifluoroacetyl)camphor, (18) 3-heptafluorobutyryl camphor, (19) 3-bromocamphor, (20) 9,10-dibromocamphor, (21) 3,9,10-tribromocamphor, (22) dicyclopentadiene, (23) methylcyclopentadiene dimer, (24) tricyclo[5.2.1]decane, (25) 4,8-bis(hydroxymethyl)tricyclo[5.2.1.0^{2.6}]decane, (26) 8-ketotricyclo[5.2.1.0^{2.6}]decane, and the like; (B) cyclobutenes and cyclobutene derivatives, of the general formula wherein R₁, R₂, R₃, R₄, R₅, and R₆ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, and R₆ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, or the like, as well as mixtures thereof.

Examples of cyclobutenes and cyclobutene derivatives include (1) 3,4-dimethoxy-3-cyclobutene-1,2-dione, (2) 3,4-diethoxy-3-cyclobutene-1,2-dione, (3) 3,4-diisopropoxy-3-cyclobutene-1,2-dione, (4) 3,4-dibutoxy-3-cyclobutene-1,2-dione, and the like;
(C) cyclopentanes and cyclopentane derivatives, and cyclopentenes and cyclopentene derivatives, of the formulae wherein R₁, R₂, R₃, R₄, R₅, R₆, R₇, R₈, R₉, and R₁₀ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, and R₁₀ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, ClO₃⁻, ClO₃⁻, or the like, as well as mixtures thereof.

Examples of cyclopentanes and cyclopentenes include (1) 3-methyl-2-(nitromethyl)-5-oxocyclopentaneacetic acid, (2) 3-ethyl-2-hydroxy-2-cyclopenten-1-one, (3) methyl-4-methoxy-2-oxo-3-cyclopentene-1-carboxylate, (4) 3,3a,6,6a-tetrahydro-2H-cyclopenta[b]furan-2-one, (5) 3a,4,5,6a-hexahydro-5-hydroxy-4(hydroxymethyl)-2H-cydopenta[b]furan-2-one, (6) 3-methyl-1,2-cyclopentanedione, (7) 4-hydroxy-5-methyl-4-cyclopentene-1,3-dione monohydrate, and the like;
(D) cyclohexane, cyclohexene, and cyclohexadiene compounds and derivatives, of the general formulae wherein R₁, R₂, R₃, R₄, R₅, R₆, R₇, R₈, R₉, R₁₀, R₁₁, and R₁₂ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, R₁₀, R₁₁, and R₁₂ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, Cl0₃⁻, or the like, as well as mixtures thereof.

Examples of cyclohexanes, cyclohexenes, and cyclohexadienes include (1) 2,4,4-trimethylcyclohexen-1-one, (2) ethyl-6-methyl-2-oxo-3-cyclohexene-1-carboxylate, (3) ethyl 4-hydroxy-6-methyl-2-oxo-3-cyclohexene-1-carboxylate, (4) 5-(1-acetoxy-1-methylethyl)-2-methyl-2-cyclohexen-1-one, (5) thymoquinone, (6) 2,6,6-trimethyl-2-cyclohexene-1,4-dione, and the like;
(E) indans and indan derivatives, including those of the general formula wherein R₁, R₂, R₃, R₄, R₅, R₆, R₇, R₈, R₉, and R₁₀ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, and R₁₀ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of indans and indan derivatives include (1) indan, (2) 1-indanol, (3) 2-indanol, (4) 1-indanone, (S) 2-indanone, and the like; (F) tetralones and tetralone derivatives, including those of the general formulae wherein R₁, R₂, R₃, R₄, R₅, R₆, R₇, R₈, R₉, and R₁₀ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, R₉, and R₁₀ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of tetralones and tetralone derivatives include (1) 2-acetyl-1-tetralone, (2) 4-methyl-1-tetralone, (3) 5,7-dimethyl-1-tetralone, (4) 6,7-dimethoxy-1-tetralone, (5) 1-methyl-2-tetralone, (6) 6,7-dimethoxy-2-tetralone, and the like;
(G) cyclonones and cyclonone derivatives, of the general formula wherein the curved portion of the structure represents a hydrocarbon chain or a substituted hydrocarbon chain, preferably of from about 3 to about 1 1 carbon atoms, wherein two or more substituents can be joined together to form a ring, and wherein the substituents on the hydrocarbon chain can be (but are not limited to) alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of cyclonones and cyclonone derivatives include (1) cyclohexanone, (2) cycloheptanone, (3) cyclooctanone, (4) cyclononanone, (5) cyclodecanone, (6) cycloundecanone, (7) cyclododecanone, (8) cyclotridecanone, (9) cyclopentadecanone, (10) 2-acetylcyclohexanone, (11) 2-allylcyclohexanone, (12) 2-phenylcyclohexanone, (13) cyclohexanedione, (14) 2-acetyl-1,3-cyclohexanedione, (15) 4,4-dimethyl-1,3-cyclohexanedione, (16) 2-acetyl-1,3-cyclopentanedione, (17) 3,3,5,5-tetramethyl-1,2-cyclopentanedione, and the like; (H) bicyclo[3.2.1]octan-2-one, (I) endo-dimethyl 7-oxabicyclo[2.2.1]heptane-2,3-dicarboxylate, (J) cineole, (K) bicyclo[2.2.2]oct-5-ene-2,3-dimethanol, (L) tropone, (M) tropolone, (N) cyclooctene oxide (9-oxabicyclo[6.1.0]nonane), (O) 1,2,5,6-diepoxycyclooctane, (P) 9-methyl-Δ⁵⁽¹⁰⁾-octalin-1,6-dione, (Q) cis-bicyclo[3.3.0]octane-3.7-dione, (R) azulene, (S) 1-benzosuberone, (T) 1,5,9-cyclododecatriene, (U) cyclododecane epoxide, (V) 2,3-cyclododeceno pyridine, (W) 1,2,5,6,9,10-hexabromo cyclododecane, (X) 8-cyclohexadecen-1-one, (Y) bicyclo[10.3.0]pentadec-12(1)-en-13-one, (Z) 1,4,4a,8a-tetrahydro-endo-1,4-methanonaphthalene-5,8-dione, and the like;

IV. Sulfur-containing compounds, including (A) thioureas and thiourea derivatives, such as (1) 1-allyl-2-thiourea, (2) 1-methallyl-3-methyl-2-thiourea, (3) 4-allyl-3-thiosemicarbazide, (4) 1,3-diethyl-2-thiourea, (5) 1,3-dibutyl-2-thiourea, (6) 1-benzyl-3-methyl-2-thiourea, (7) 1,1,3,3-tetramethyl-2-thiourea, (8) 2-imino-4-thiobiuret, (9) 1-allyl-3-(2-hydroxyethyl)-2-thiourea, (10) S-(2-aminoethyl)isothiouronium bromide hydrobromide, (11) S,S-diphenylsulfillimine monohydrate, and the like; (B) sulfones and sulfone derivatives, such as (1) methylsulfone (dimethylsulfone), (2) ethylsulfone (diethylsulfone), (3) butylsulfone (dibutylsulfone), (4) butadiene sulfone, (5) tetramethylene sulfone, (6) 1,4-butane sulfone, (7) 1,4-butanediolcyclic sulfate, (8) benzylsulfone, (9) phenylsulfone (diphenylsulfone), (10) phenylvinylsulfone, (11) phenylstyrenesulfone, (12) phenyl-2-(trimethylsilyl)methyl sulfone, (13) phenyl 2-(trimethylsilyl)ethyl sulfone, (14) phenyl 2-(trimethylsilyl)ethynyl sulfone, (15) 4-(fluorophenyl)sulfone, (16) 4-(fluorophenyl)methyl sulfone, (17) chloromethylphenyl sulfone, (18) chloromethyl-p-tolyl sulfone, (19) 2-chloroethylphenyl sulfone, (20) methylthiomethylphenyl sulfone, (21) methylthiomethyl-p-tolyl sulfone, (22) 2-(phenylsulfonyl) tetrahydropyran, (23) 1-(phenylsulfonyl)indole, (24) 1-(p-toluenesulfonyl)imidazole, (25) 1-(p-tosyl)-3,4,4-trimethyl imidazolidine, (26) 4-(p-tosylsulfonyl)hexahydro -1,4-thiazepine, and the like; (C) thiocyclic compounds, such as (1) thionaphthene, (2) 4-keto-4,5,6,7-tetrahydrothianaphthene, (3) 2,2'-bithiophene, (4) 2,2':5',2"-terthiophene, (5) D,L-N-acetylhomocysteine thiolactone, (6) tetrahydrothiopyran-4-one, (7) thiochroman-4-one, (8) thiochroman-4-ol, (9) D,L-thioctic acid, (10) ethyl 1,3-dithiolane-2-carboxylate, (11) 3H-1,2-benzodithiol-3-one, (12) 1,3-dithiane, (13) 2-phenyl-1,3-dithiane, (14) ethyl-1,3-dithiane-2-carboxylate, (15) 5,6-dihydro-5-methyl-4H-1,3,5-dithiazine, (16) 1,4-dithiane, (17) 2,5-dihydroxy-2,5-dimethyl-1,4-dithiane, (18) 1,5-dithiacyclooactan-3-ol, (19) 1,4-dithiaspiro [45] decan-8-ol, (20) 1,3,5-trithiane, (21) 1,4,7-trithiacyclononane, (22) 1,4,7-trithiacyclodecane, (23) 1,4,7,10-tetrathiacyclododecane, (24) 3,6,9,14-tetrathiabicyclo [9.2.1] tetradeca-11,13-diene, (25) 1,4,8,1-tetrathiacyclotetradecane, (26) 1,5,9,13-tetrathiocyclohexadecane, (27) 1,5,9,13-tetrathiacyclohexadecane-3,11-diol, (28) 1,4,7,10,13-pentathiacyclopentadecane, (29) 1,4,7,10,13,16-hexathiacyclooctadecane, (30) 1,5,9,13,17,21-hexathiacyclotetracosane-3,11,19-triol, (31) 1,4,7,10,13,16,19,22-octathiacyclotetracosane, (32) 1,4,8,11,15,18,22,25-octathiacyclooctacosane, (33) 1,4,7,10,13,16,19,22,25-nonathiacycloheptacosane, and the like; (D) sulfites and sulfite derivatives, including (1) dimethylsulfite, (2) diethylsulfite, (3) sodium sulfite, and the like; (E) sulfides and sulfide derivatives, including (1) allyldisulfide, (2) aminophenyldisulfide, (3) benzyldisulfide, (4) benzylphenylsulfide, and the like; (F) quaternary sulfur compounds and their derivatives, including (1) trimethylsulfonium methylsulfate, (2) (2-chloroethyl)dimethylsulfonium iodide, (3) 3-(chloropropyl)diphenylsulfonium tetrafluoroborate, (4) trimethyl sulfonium iodide, (5) trimethyl sulfoxonium iodide, (6) trimethyl sulfoxonium chloride, (7) triphenyl methane sulfenyl chloride, (8) dimethyl (2-methoxy-5-nitrobenzyl) sulfonium bromide, (9) thionin perchlorate, (10) p-xylylene bis(tetrahydrothiopheneum chloride), (11) tris (dimethyl amino) sulfonium difluorotrimethyl silicate, (12) tris (dimethyl amino) sulfonium trifluoromethoxide, (13) (3-amino-3-carboxypropyl) dimethyl sulfonium chloride, and the like;

V. Thia-aza-cyclic compounds, including (A) thiazoles and thiazole derivatives, and thiazolidines and thiazolidine derivatives, and thiadiazoles and thiadiazole derivatives, including those of the general formulae wherein R₁, R₂, R₃, R₄, R₅, R₆, and R₇ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, and R₇ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ⁻, wherein n is an integer of 1, 2, or 3, x is a number indicating the relative ratio between compound and acid (and may be a fraction), and Y is an anion, such as Cl⁻, Br⁻, l⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, lO₃⁻, ClO₃⁻, or the like, as well as mixtures thereof.

Examples of thiazoles include (1) 2-amino-2-thiazoline, (2) 2-amino thiazole, (3) 2-amino-4-methylthiazole, (4) 2-amino-4-methylthiazole, (S) 2-amino-4-thiazoleacetic acid, (6) 2-acetamido-4-methylthiazole, (7)2-acetylthiazole, (8) 5-acetyl-2,4-dimethylthiazole, (9) 4-methyl-5-vinylthiazole, (10) 2-amino-4-phenyl-5-tetradecylthiazole, (11) 2,4-thiazolidine dione, (12) 3-aminorhodanine, (13) 3-methylrhodanine, (14) 3-ethylrhodanine, (15) 3-allylrhodanine, (16) 3-hydroxy-4-methyl-2(3H)-thiazolethione, (17) benzothiazole, (18) 2-methylbenzothiazole, (19) 2-(methylthio)benzothiazole, (20) 2-amino-4-methylbenzothiazole, (21) 3-methylbenzothiazole-2-thione, (22) 2,1,3-benzothiadiazole, (23) 4-amino-2,1,3-benzothiadiazole, (24) 3,4-dimethyl-5-(2-hydroxyethyl)thiazolium iodide, (25) 3-ethyl-5-(2-hydroxyethyl)4-methylthiazolium bromide, (26) 2-amino-5-nitrothiazole, (27) 2-amino-α-(methoxyimino)-4-thiazole acetic acid, (28) ethyl 2-amino-α-(hydroxyimino)-4-thiazole acetate, (29) ethyl 2-amino-α-(methoxyimino)-4-thiazole acetate, (30) ethyl 2-amino-4-thiazole acetate, (31) ethyl 2-amino-4-thiazole glyoxylate, (32) 1-phenyl-3-(2-thiazolyl)-2-thiourea, (33) 2-amino-4-methoxy benzothiazole, (34) 2-amino-5,6-dimethylbenzothiazole, (35) N'-(2-thiazolyl) sulfanilamide, (36) 6-ethoxy-2-benzothiazole sulfonamide, (37) ethyl-2-(formylamino)-4-thiazoleacetate, (38) ethyl-2-(formylamino)-4-thiazoleglyoxylate, (39) 2-(formylamino)-α-(methoxyimino)-4-thiazole acetic acid, (40) 2-acetamido-4-methyl-5-thiazole sulfonyl chloride, (41) (4R)-(-)-2-thioxo-4-thiazolidine carboxylic acid, (42) (R)-(-)-thiazolidine-4-carboxylic acid, (43) pseudothiohydantoin, (44) 2-amino-1,3,4-thiadiazole, (45) 2-amino-5-trifluoromethyl-1,3,4-thiadiazole, (46) 2-amno-5-methyl-1,3,4-thiadiazole, (47) 2-amino-5-ethyl-1,3,4-thiadiazole, (48) 2-amino-5-(ethylthio)-1,3,4-thiadiazole, (49) 5-amino-1,3,4-thiadiazole-2-thiol, (50) 2-acetamido-5-benzyl thio-1,3,4-thiadiazole, (51) 5-acetamido-1,3,4-thiadiazole-2-sulfonamide, (52) 5-anilino-1,2,3,4-thiatriazole, (53) 2-amino-4,5-dimethyl thiazole hydrochloride, (54) 2-amino 4-imino-2-thiazoline hydrochloride, (55) 2-amino-2-thiazoline hydrochloride, (56) 2-amino-5-bromothiazole monohydrobromide, (57) 5-amino-3-methyl isothiazole hydrochloride, (58) 3-methyl-2- benzothiazolinone hydrazone hydrochloride hydrate, (59) 5-amino-2-methylbenzothiazole dihydrochloride, (60) 2,4-diamino-5-phenyl thiazole monohydrobromide, (61) 2-amino-4-phenyl thiazole hydrobromide monohydrate, (62) 2-(tritylamino)-a-(methoxyimino)-4-thiazole acetic acid hydrochloride, (63) (2,3,5,6-tetrahydro-6-phenylimidazo [2,1-b] thiazole hydrochloride, (64) 3-ethyl-2-methyl-2-thiazolium iodide, (65) 3-benzyl-5-(2-hydroxyethyl)-4-methyl thiazolium chloride, (66) thiamine hydrochloride, (67) 3-(carboxymethyl) benzothiazolium bromide, (68) 2-azido-3-ethyl benzothiazolium tetrafluoroborate, (69) 3-ethyl-2-methyl benzothiazolium iodide, (70) 2-methyl-3-propyl benzothiazolium iodide, (71) 3-ethyl-2-(2-hydroxy-1-propenyl) benzothiazolium chloride, (72) 3,6-dimethyl-2-(4-dimethyl aminophenyl) benzothiazolium bromide, and the like; (b) phenothiazines, including those of the general formula wherein R₁, R₂, R₃, R₄, R₅, R₆, R₇, R₈, and R₉ each, independently of the others, can be (but are not limited to) hydrogen atoms, alkyl groups, preferably with from 1 to about 6 carbon atoms and more preferably with from 1 to about 3 carbon atoms, substituted alkyl groups, preferably with from 1 to about 12 carbon atoms and more preferably with from 1 to about 6 carbon atoms, aryl groups, preferably with from about 6 to about 24 carbon atoms and more preferably with from about 6 to about 12 carbon atoms, substituted aryl groups, preferably with from about 6 to about 30 carbon atoms and more preferably with from about 6 to about 18 carbon atoms, arylalkyl groups, preferably with from about 7 to about 31 carbon atoms and more preferably with from about 7 to about 20 carbon atoms, substituted arylalkyl groups, preferably with from about 7 to about 32 carbon atoms and more preferably with from about 7 to about 21 carbon atoms, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more of R₁, R₂, R₃, R₄, R₅, R₆, R₇, R₈, and R₉ can be joined together to form a ring, and wherein the substituents on the substituted alkyl groups, substituted aryl groups, and substituted arylalkyl groups can be (but are not limited to) hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, azide groups, and the like, wherein two or more substituents can be joined together to form a ring. Other variations are also possible, such as a double bond between one of the ring carbon atoms and another atom, such as carbon, oxygen, or the like. These compounds can also be in acid salt form, wherein they are associated with a compound of the general formula xHₙYₙ-, wherein n is an integer of 1, 2, or 3, x is a number indicating the relative ratio between compound and acid (and may be a fraction), and Y is an anion, such as Cl⁻, Br⁻, L⁻, HSO₄⁻, SO₄²⁻, NO₃⁻, HCOO⁻, CH₃COO⁻, HCO₃⁻, CO₃²⁻, H₂PO₄⁻, HPO₄²⁻, PO₄³⁻, SCN⁻, BF₄⁻, ClO₄⁻, SSO₃⁻, CH₃SO₃⁻, CH₃C₆H₄SO₃⁻, SO₃²⁻, BrO₃⁻, IO₃⁻, ClO₃⁻, or the like, as well as mixtures thereof.

Examples of phenothiazines include (1) trifluoroperazine dihydrochloride, (2) thioridazine hydrochloride, (3) (±)-promethazine hydrochloride, (4) ethopropazine hydrochloride, (5) chlorpromazine hydrochloride, and the like;

VI. Phosphorus compounds and their derivatives, including (A) phosphines, such as (1) trialkyl, triaryl, and heterocyclic phosphines and their derivatives, including (a) triphenylphosphine, (b) tri-m-tolyl phosphine, (c) tris(3-methoxyphenyl)phosphine, (d) tris(4-chlorophenyl)phosphine, (e) tris(pentafluorophenyl)phosphine, (f) tricyclohexylphosphine, (g) tribenzylphosphine, (h) tri-2-furylphosphine, (i) bis (pyrrolidino)methoxy phosphone, (j) compounds of the general formula (C₆H₅)₂P(CH₂)nP(C₆H₅)₂ where n is an integer of from 0 to about 10, such as (1) n=0: tetraphenylbiphosphine, (2) n = 3: 1,3-bis(diphenylphosphino)propane, (3) n = 5: 1,5-bis(diphenylphosphino)pentane, (4) n = 6: 1,6-bis(diphenylphosphino)hexane, and the like; (k) alkyldiphenyl or dialkylphenyl compounds, including (1) isopropyl diphenyl phosphine, (2) diphenyl (p-tolyl) phosphine, (3) (4-bromophenyl) diphenyl phosphine, (4) diphenyl-2-pyridylphosphine, (5) dicyclohexylphenyl phosphine, and the like; (B) phosphites and phosphite derivatives, including (1) trialkyl and triaryl phosphites and their complexes, such as (a) trimethyl phosphite, (b) triethyl phosphite, (c) tris(2-chloroethyl) phosphite, (d) tributyl phosphite, (e) triphenyl phosphite,(f) trimethyl phosphite copper iodide, (g) triethyl phosphite copper iodide, and the like; (2) dialkyl and diaryl phosphites, such as (a) dipropyl phosphite, (b) bis(2-ethylhexyl) phosphite, (c) bis(4-nitrobenzyl) phosphite, (d) 2,2'-ethylidene bis(4,6-di-tert-butylphenyl) fluorophosphite, (e) pentaerythritol diphenyl diphosphite, and the like; (C) cyclic phosphorus compounds, including (1) 2-furyltetramethyl phosphorodiamidate, (2) diethyl(pyrrolidinomethyl)phosphonate, (3) cyclophosphamide monohydrate, (4) 2-chloro-1,3,2-dioxaphospholane-2-oxide, (5) N,N-diethyl-1,5-dihydro-2,4,3-benzodioxaphosphepin-3-amine, (6) 1,2-phenylene phosphochloridite, (7) 1,2-phenylene phosphochloridate, (8) 2-chloro-4H-1,3,2-benzodioxaphosphorin-4-one, (9) 2,4-bis(methylthio)-1,3-dithia-2,4-diphosphetane-2,4-disulfide, and the like; (D) phosphine oxide compounds, including (1) trisubstituted phosphine oxides, such as (a) triphenyl phosphine oxide, (b) tris(hydroxymethyl) phosphine oxide, (c) trimethoxy phosphine oxide, (d) triethoxy phosphine oxide, (e) triphenoxy phosphine oxide, (f) tris (2-butoxy ethoxy) phosphine oxide, and the like; (2) disubstituted phosphine oxides, such as (a) diphenyl phosphine oxide, (b) diphenyl (2,4,6-trimethylbenzoyl) phosphine oxide, and the like; (3) hydroxy phosphine oxide compounds, such as (a) phenyl phosphinic acid, (b) diphenyl phosphate, (c) vinyl phosphonic acid, (d) propyl phosphonic acid, (e) pyrophosphoric acid, (f) triphenylphosphate, and the like; (E) quaternary phosphonium salts, including (1) tetrabutylphosphonium chloride, (2) tetrabutylphosphonium bromide, (3) hexadecyltributylphosphonium bromide, (4) stearyltributylphosphonium bromide, (5) azidotris(diethylamino)phosphonium bromide, (6) phosphonitrilic chloride trimer, (7) tetramethyl phosphonium bromide, (8) tetramethyl phosphonium chloride, (9) tetraethyl phosphonium bromide, (10) tetraethyl phosphonium chloride, (11) tetraethyl phosphonium iodide, (12) tetraphenyl phosphonium bromide, (13) tetraphenyl phosphonium chloride, (14) tetraphenyl phosphonium Iodide, (15) methyl triphenyl phosphonium bromide, (16) methyl triphenyl phosphonium iodide, (17) ethyl triphenyl phosphonium bromide, (18) n-propyl triphenyl phosphonium bromide, (19) isopropyl triphenyl phosphonium iodide, (20) cyclopropyl triphenyl phosphonium bromide, (21) n-butyl triphenyl phosphonium bromide, (22) isobutyl triphenyl phosphonium bromide, (23) hexyl triphenyl phosphonium bromide, (24) benzyl triphenyl phosphonium chloride, (25) bromomethyl triphenyl phosphonium bromide, (26) chloromethyl triphenyl phosphonium chloride, (27) 3-bromopropyl triphenyl phosphonium bromide, (28) 3-bromobutyl triphenyl phosphonium bromide, (29) 4-bromobutyl triphenyl phosphonium bromide, (30) 2-dimethyl aminoethyl triphenyl phosphonium bromide, (31) [(3-dimethyl amino) propyl] triphenyl phosphonium bromide, (32) 2-hydroxyethyl triphenyl phosphonium bromide (33) (2-hydroxyethyl) triphenyl phosphonium chloride, (34) [(R)-(+)-3-hydroxy-2-methyl propyl] triphenyl phosphonium bromide, (35) [(S)-(-)-3-hydroxy-2-methyl propyl] triphenyl phosphonium bromide, (36) (2-hydroxybenzyl triphenyl phosphonium bromide, (37) (formyl methyl) triphenyl phosphonium chloride, (38) (methoxymethyl) triphenyl phosphonium chloride, (39) acetonyl triphenyl phosphonium chloride, (40) carbomethoxymethyl triphenyl phosphonium bromide, (41) (ethoxy carbonyl methyl) triphenyl phosphonium chloride, (42) carbethoxymethyl triphenyl phosphonium bromide, (43) (tert-butoxy carbonyl methyl) triphenyl phosphonium bromide, (44) phenacyl triphenyl phosphonium bromide, (45) (4-ethoxybenzyl) triphenyl phosphonium bromide, (46) 4-butoxybenzyl triphenyl phosphonium bromide, (47) 2-(1,3-dioxan-2-yl) ethyl] triphenyl phosphonium bromide, (48) (1,3-dioxolan-2-ylmethyl) triphenyl phosphonium bromide, (49) vinyl triphenyl phosphonium bromide, (50) allyl triphenyl phosphonium bromide, (51) allyl triphenyl phosphonium chloride, (52) propargyl triphenyl phosphonium bromide, (53) (3-trimethyl silyl-2-propynyl) triphenyl phosphonium bromide, (54) p-xylylene bis (triphenyl phosphonium bromide), and the like;

VII. Nitrile compounds and their derivatives, including (1) cyanoacetohydrazide, (2) 4,4-dimethyl-3-oxopentanenitrile, (3) 1-cyano-N-methylthioformamide, (4) cyanomethyl N,N-dimethyl dithiocarbamate, (5) 4-hydroxy-3-methoxy-phenyl acetonitrile, (6) tosyl cyanide, (7) tosylmethyl isocyanide, (8) 5-fluoro-2-methyl benzonitrile, (9) 2-fluoro-5-methyl benzonitrile, (10) 4-(methylthio) benzonitrile, (11) 4-(dimethylamino) benzonitrile, (12) 3,4-dimethoxy benzonitrile, (13) 4-hydroxy-3-methoxy benzonitrile, (14) 4-(trans-4-pentyl cyclohexyl)benzonitrile, (15) 4'-pentyl-4'-biphenyl carbonitrile, (16) 4'-(pentyloxy)-4-biphenylcarbonitrile, (17) 4'-hexyl-4-biphenyl carbonitrile, (18) 4'-(hexyloxy)-4-biphenyl carbonitrile, (19) 4'-heptyl-4-biphenyl carbonitrile, (20) 4'-heptyloxy-4-biphenyl carbonitrile, (21) 4'-octyl-4-biphenyl carbonitrile, (22) 4'-(octyloxy)-4-biphenyl carbonitrile, (23) succinonitrile, (24) fumaronitrile, (25) 1,4-dicyano-2-butene, (26) (dimethyl aminomethylene)malononitrile, (27) (1-ethoxyethylidene)malononitrile, (28) α-chlorobenzylidenemalononitrile, (29) benzylidenemalononitrile, (30) 2-benzoyloxy-2-phenyl malononitrile, (31) O-(p-tosyl)isonitrosomalononitrile, (32) tetrafluorophthalonitrile, (33) iminodiacetonitrile, (34) phenylene diacetonitrile, (35) 3,3'-(4-formyl phenylimino) dipropionitrile, (36) tris (2-cyanoethyl) nitromethane, (37) 1,1,3,3-propanetetracarbonitrile, (38) tetracyanoethylene oxide, and the like;

VIII. Isothiocyanate compounds and isocyanate compounds and their derivatives, including (A) 4-azidophenyl isothiocyanate, (B) 1-naphthyl isothiocyanate, (C) 4-dimethyl amino-1-naphthyl isothiocyanate, (D) 1-isothiocyanato-4-(trans-4-propyl cyclohexyl) benzene, (E) 1-(trans-4-hexyl cyclohexyl)-4-isothiocyanato benzene, (F) 1-(4-trans-hexyl cyclohexyl)-4-[2-(4-isothio cyanatophenyl)] benzene, (G) 1-isothiocyanato-4-(trans-4-octylcyclohexyl) benzene, (H) 4-isothiocyanatophenyl-4-pentabicyclo [2.2.2] octane-1-carboxylate, (I) benzylthiocyanate, (J) guanidinethiocyanate, (K) methylene dithiocyanate, (L) 4,4'-methylene bis (phenyl isocyanate), (M) 4,4'-methylene bis(2,6-diethyl isocyanate), and the like;

IX. Oxime compounds and their derivatives, including (A) formamidoxime, (B) acetaldoxime, (C) pyruvic aldehyde-1-oxime, (D) acetone oxime, (E) ethylchlorooximido acetate, (F) 2,3-butane dione monoxime, (G) 5-hydroxy pentenal oxime, (H) cyclopentanone oxime, (I) cyclohexanone oxime, (J) cyclooctanone oxime, (K) benzaldehyde oxime, (L) 2-nitrobenzaldehyde oxime, (M) salicyl aldoxime, (N) 2-isonitroso acetphenone, (O) 1-phenyl-1,2-propanedione 2-oxime, (P) 2-pyridine aldoxime, (Q) nifuroximeand the like;

X. Hydroxamic acid derivatives, including (A) acetohydroxamic acid, (B) suberohydroxamic acid, (C) mandelohydroxamic acid, (D) benzohydroxamic acid, (E) N-phenylbenzohydroxamic acid, and the like;

XI. Halide compounds, including (A) tetraalkyl ammonium salts, such as (1) tetramethylammonium fluoride tetrahydrate, (2) tetraethylammonium acetate tetrahydrate, (3) tetrabutylammonium chloride, (4) tetrabutylammonium chloride hydrate, (5) tetrabutylammonium bromide, (6) tetrabutylammonium tribromide, (7) tetrabutylammonium acetate, (8) tetrabutylammonium thiocyanate, (9) tetrapentylammonium bromide, (10) tetrahexylammonium bromide, (11) tetrahexylammonium chloride, (12) tetrahexylammonium hydrogensulfate, (13) tetraheptylammonium chloride, (14) tetraheptylammonium bromide, (15) tetraoctylammonium bromide, (16) tetrakisdecylammonium bromide, (17) tetrahexadecylammonium bromide, (18) tetramethyl ammonium bromide, (19) tetramethyl ammonium chloride, (20) tetramethyl ammonium iodide, (21) tetraethyl ammonium bromide, (22) tetraethyl ammonium chloride, (23) tetraethyl ammonium iodide, (24) tetrapropyl ammonium bromide, (25) tetrapropyl ammonium iodide, (26) tetrabutyl ammonium iodide, (27) tetrapentyl ammonium chloride, (28) tetrahexyl ammonium bromide, (29) tetrahexyl ammonium iodide, (30) tetradecyl ammonium bromide, (31) tetradodecyl ammonium bromide, (32) tetraoctadecyl ammonium bromide, and the like; (B) alkyl trialkyl ammonium salts, aryl trialkyl ammonium salts, alkyl triaryl ammonium salts, and aryl triaryl ammonium salts, such as (1) methyltrioctylammonium bromide, (2) tridodecylmethylammonium chloride, (3) tridodeylmethylammonium iodide, (4) (-)-N-dodecyl-N-methylephedrinium bromide, (5) phenyltrimethylammonium tribromide, (6) tricapryl methyl ammonium chloride, (7) tridodecyl methyl ammonium chloride, (8) tridecyloxypropyl dihydroxy ethyl methyl ammonium chloride, (9) N-tetradecyl dimethyl-naphthyl methyl ammonium chloride, (10) octadecyl diethanol methyl ammonium chloride, (11) octadecyl dihydroxyethyl methyl ammonium chloride, (12) dihydrogenated tallow benzyl methyl ammonium chloride, (13) 2-aminoethyl trimethyl ammonium chloride hydrochloride, (14) 2-bromoethyl trimethyl ammonium bromide, (15) 2-chloroethyl trimethyl ammonium chloride, (16) 3-carboxypropyl trimethyl ammonium chloride, (17) [3-(methacryloyl amino) propyl] trimethyl ammonium chloride, (18) phenyl trimethyl ammonium bromide, (19) phenyl trimethyl ammonium chloride, (20) phenyl trimethyl ammonium iodide, (21) benzyl trimethyl ammonium chloride, (22) benzyl trimethyl ammonium bromide, (23) 4-nitrobenzyl trimethyl ammonium chloride, (24) [2-(4-nitrophenyl) allyl] trimethyl ammonium iodide, (25) coco trimethyl ammonium chloride, (26) palmityl trimethyl ammonium chloride, (27) myristyl trimethyl ammonium bromide, (28) oleyl trimethyl ammonium chloride, (29) soya trimethyl ammonium chloride, (30) tallow trimethyl ammonium chloride, (31) hydrogenated tallow trimethyl ammonium chloride, (32) stearyl trimethyl ammonium chloride, (33) behenyl trimethyl ammonium chloride, (34) guar hydroxypropyl trimethyl ammonium chloride, (35) benzyl triethyl ammonium chloride, (36) benzyl triethyl ammonium bromide, (37) butyl tripropyl ammonium bromide, (38) methyl tributyl ammonium chloride, (39) methyl tributyl ammonium bromide, (40) methyl tributyl ammonium iodide, (41) benzyl tributyl ammonium chloride, (42) benzyl tributyl ammonium bromide, (43) benzyl tributyl ammonium iodide, (44) heptyl tributyl ammonium bromide, and the like; (C) dialkyl dialkyl ammonium salts, such as (1) benzyldodecyldimethylammonium bromide, (2) benzyltetradecyldimethylammonium chloride dihydrate, (3) benzylcetyldimethylammonium chloride monohydrate, (4) benzylstearyldimethylammonium chloride monohydrate, (5) N,N-dimethyl methylene ammonium chloride, (6) N,N-dimethyl methylene ammonium iodide, (7) chloromethylene dimethyl ammonium chloride, (8) dichloromethylene dimethyl ammonium chloride, (9) dimethyl amino methylene amino methylene dimethyl ammonium chloride, (10) benzethonium chloride, (11) methyl benzethoniumchloride, (12) 1-propanaminium 2,3-dihydroxy-N-dimethyl-N-[3(oxococoyl) amino]propyl]-chloride, (13) cetyl dimethyl ethyl ammonium bromide, (14) octyl dodecyl dimethyl ammonium chloride, (15) dodecyl (2-hydroxy1-methyl-2-phenyl-ethyl) dimethyl ammonium bromide, (16) dodecyl dimethyl 2-phenoxyethyl ammonium bromide, (17) dodecanoyl-N-methylamino ethyl-(phenyl carbamyl methyl) dimethyl ammonium chloride, (18) 3-chloro-2-hydroxypropyl N,N,N-dimethyl dodecyl ammonium chloride, (19) 3-chloro-2-hydroxypropyl N,N,N-dimethyl octadecyl ammonium chloride, (20) dodecyl benzyl dimethyl ammonium bromide, (21) dodecyl benzyl dimethyl ammonium chloride, (22) coco benzyl dimethyl ammonium chloride, (23) benzyl tetradecyl dimethyl ammonium chloride, (24) benzyl cetyl dimethyl ammonium chloride, (25) benzyl octadecyl dimethyl ammonium chloride, (26) benzyl tallow dimethyl ammonium chloride, (27) benzyl hydrogenated tallow dimethyl ammonium chloride, (28) benzyl behenyl dimethyl ammonium chloride, (29) dioctyl dimethyl ammonium chloride, (30) didecyl dimethyl ammonium chloride, (31) didecyl dimethyl ammonium bromide, (32) dicoco dimethyl ammonium chloride, (33) dicetyl dimethyl ammonium chloride, (34) disoya dimethyl ammonium chloride, (35) ditallow dimethyl ammonium chloride, (36) dihydrogenated tallow dimethyl ammonium chloride, (37) dibehenyl/diarachidyl dimethyl ammonium chloride, (38) soya amido propyl benzyl dimethyl ammonium chloride, (39) soya dicoco quaternary ammonium chloride, (40) gluconamidopropyl dimethyl-2-hydroxyethyl ammonium chloride, (41) N-alkyl-N-N-dimethyl-N(dodecyl acetate) ammonium chloride, wherein alkyl has from 14 to 20 carbon atoms, (42) mink amidopropyl dimethyl-2-hydroxyethyl ammonium chloride, (43) N-rapeseed-(3-amidopropyl)-N-N-dimethyl-N-(2,3 epoxy propyl) ammonium chloride, (44) N-stearyl-(3-amido propyl)-N-benzyl dimethyl ammonium chloride, (45) rapeseed amido propyl benzyl dimethyl ammonium chloride, (46) rapeseed amido propyl ethyl dimethyl ammonium chloride, (47) cocamidopropyl polyethylene glycol dimethyl ammonium chloride phosphate, and the like; (D) choline salts, such as butyrylcholine chloride, and the like.

Any other transparentizing agent suitable for the selected migration marking material(s) can also be employed, as well as mixtures thereof.

### EXAMPLE I

Migration imaging members were prepared as follows. A solution for the softenable layer was prepared by dissolving about 84 parts by weight of a terpolymer of styrene/ethylacrylate/acrylic acid (prepared as disclosed in U.S. Patent 4,853,307, and about 16 parts by weight of N,N'-diphenyl-N,N'-bis(3"-methylphenyl)-(1,1'-biphenyl)-4,4'-diamine (prepared as disclosed in U.S. Patent 4,265,990, in about 450 parts by weight of toluene. N,N'-diphenyl-N,N'-bis(3''-methylphenyl)-(1,1'-biphenyl)-4,4'-diamine is a charge transport material capable of transporting positive charges (holes). The resulting solution was coated by a solvent extrusion technique onto 3 mil thick polyester substrates (Melinex 442), aluminized to 50 percent light transmission), and the deposited softenable layers were allowed to dry at about 115°C for about 2 minutes, resulting in dried softenable layers with thicknesses of about 4 microns. The temperature of the softenable layers was then raised to about 115°C to lower the viscosity of the exposed surfaces of the softenable layers to about 5×10³ poises in preparation for the deposition of marking material. Thin layers of particulate vitreous selenium were then applied by vacuum deposition in a vacuum chamber maintained at a vacuum of about 4×10⁻⁴ Torr. The imaging members were then rapidly chilled to room temperature. Reddish monolayers of selenium particles having an average diameter of about 0.3 micron embedded about 0.05 to 0.1 micron below the surfaces of the copolymer layers were formed.

Separate sheets of polyester 100 microns thick were solvent coated from solutions of toluene containing about 10 percent by weight solids with blends of various transparentizing agents as indicated in the tables below with a styrene/ethyl acrylate/acrylic acid binder (obtained from Scientific Polymer Products, #815) to form coating layers about 4 microns thick. The weight ratio of transparentizing agent to binder was 1:4 in each instance. The coated sheets were dried at 25°C for 1 hour. Thereafter, the coated surfaces of the polyester sheets were placed in intimate contact with the surfaces of the migration imaging members coated with the softenable material and the migration marking material, and the "sandwiches" thus formed were subjected to temperatures of 100°C for 1 minute, at which temperature the softenable layer was softened sufficiently to enable contact between the embedded selenium particles and the transparentizing agents while the softenable material was in a molten state. The polyester sheets coated with the transparentizing agents were then separated from the migration imaging members and the UV absorption spectra at 685 nm of the migration imaging members were measured to determine the extent of migration marking material transparentization. UV absorption spectra were measured with a Shimadzu UV-160 spectrometer; all spectra were recorded by using 50% transmission aluminized ICI 442 polyester as a reference. The optical densities of the migration imaging members were also measured with a Macbeth TR927 densitometer in the visible, ultraviolet, and infrared range, using a Wratten No. 47 filter for the blue measurements, a Wratten No. 18A filter for the UV measurements, and a Wratten No. 25 filter for the IR measurements. For comparison purposes, the UV absorption spectrum at 685 nm and the optical density of the migration imaging members prior to contact with the sheet coated with transparentizing agent were also measured. The results were as follows:

| Agent | UV absorption | Optical Density | | |
|---|---|---|---|---|
| | | vis. | UV | IR |
| none | 1.50 | 1.82 | 2.65 | 0.89 |
| piperidine thiocyanate | 0.00 | 0.40 | 1.30 | 0.70 |
| 2-piperidine methanol | 0.50 | 0.65 | 0.50 | 0.36 |
| bis(pentamethylene) urea | 0.00 | 0.27 | 0.60 | 0.35 |
| 4,4'-trimethylene bis(1-piperidine propionitrile) | 0.00 | 0.25 | 0.60 | 0.50 |
| tripiperidino phosphine oxide | 0.00 | 0.24 | 0.55 | 0.35 |
| homopiperazine | 0.00 | 0.30 | 0.55 | 0.32 |
| 1-piperonyl piperazine | 0.00 | 0.28 | 1.09 | 0.30 |
| hexacyclentrisulfate | 0.50 | 0.60 | 1.20 | 0.70 |
| 5,10,15,20-tetraphenyl-21*H* ,23*H* porphine | 0.40 | 1.00 | 1.50 | 0.80 |
| 5,10,15,20-tetrakis(4-methoxyphenyl)-2*H* ,23*H* -porphine | 0.70 | 1.00 | 1.50 | 1.10 |
| pyrrole-2-carboxaldehyde | 0.00 | 0.28 | 0.76 | 0.35 |
| 3-pyrrolidino-1,2-propanediol | 0.00 | 0.25 | 0.95 | 0.31 |
| pyrazole | 0.50 | 0.38 | 0.79 | 0.45 |
| 3-aminopyrazole | 0.10 | 0.41 | 1.00 | 0.50 |
| imidazole | 1.00 | 0.60 | 1.10 | 0.60 |
| 2-ethylimidazole | 0.00 | 0.35 | 0.55 | 0.38 |
| 2-(2-piperidinoethyl) pyridine | 0.00 | 0.25 | 0.75 | 0.28 |
| 1-dodecyl pyridinium chloride | 0.00 | 0.32 | 0.83 | 0.27 |
| pyridinium bromide perbromide | 0.00 | 0.11 | 0.90 | 0.19 |
| 3-aminoquinoline | 0.20 | 0.45 | 0.97 | 0.48 |
| 8-hydroxyquinoline | 0.40 | 0.40 | 0.85 | 0.50 |
| 8-hydroxyquinaldine | 0.10 | 0.40 | 0.72 | 0.55 |
| quinoxaline | 0.00 | 0.30 | 0.57 | 0.37 |
| 4,5-dihydro-6-methyl-3(2*H* )-pyridazinone monohydrate | 1.00 | 0.80 | 1.50 | 0.70 |
| phthalazine | 0.50 | 0.45 | 0.97 | 0.48 |
| 1,10-phenanthroline | 0.20 | 0.41 | 1.30 | 0.45 |
| 1,3,5-triazine | 0.00 | 0.50 | 0.97 | 0.52 |
| trichloromelamine | 0.00 | 0.15 | 0.57 | 0.09 |
| trichloroisocyanouric acid | 0.00 | 0.11 | 0.55 | 0.08 |
| norbornane | 0.05 | 0.34 | 0.85 | 0.44 |
| tricyclo[5.2.1.0] decane | 0.00 | 0.26 | 0.53 | 0.35 |
| norcamphor | 0.00 | 0.37 | 0.51 | 0.39 |
| tropolone | 0.00 | 0.28 | 3.55 | 0.08 |
| 1-indanol | 0.00 | 0.20 | 0.40 | 0.33 |
| *trans,trans,cis-* 1,5,9-cyclododecatriene | 0.00 | 0.23 | 0.80 | 0.30 |
| cyclodecane epoxide | 0.00 | 0.26 | 0.50 | 0.33 |
| 2,3-cyclododecane pyridine | 0.50 | 0.71 | 0.50 | 0.33 |
| 1,2,5,6,9,10-hexabromo-cyclododecane | 0.00 | 0.35 | 0.85 | 0.35 |
| 1,4,4a,8a-tetrahydro-endo-1,4-methanonaphthalene-5,8-dione | 0.10 | 0.39 | 1.41 | 0.43 |
| γ-butyrolactone | 0.00 | 0.62 | 0.94 | 0.63 |
| β,β-dimethyl-γ-(hydroxymethyl)-γ-butyrolactone | 0.30 | 0.42 | 1.20 | 0.50 |
| 2,5-dimethyl-4-hydroxy-3(2 *H* )-furanone | 0.00 | 0.28 | 0.65 | 0.35 |
| hydrindantin dihydrate | 0.33 | 0.60 | 1.00 | 0.65 |
| 2,4,8,10-tetraoxaspiro [5.5]undecane | 0.00 | 0.27 | 0.65 | 0.35 |
| 1,3,5-trioxane | 0.00 | 0.26 | 0.50 | 0.35 |
| cyclooctanone | 0.00 | 0.27 | 0.48 | 0.33 |
| piperonal | 0.00 | 0.25 | 0.90 | 0.28 |
| piperonylalcohol | 0.00 | 0.31 | 0.88 | 0.40 |
| piperonyl nitrile | 0.00 | 0.25 | 0.40 | 0.35 |
| 3,4(methylenedioxy) phenylacetonitrile | 0.10 | 0.40 | 0.75 | 0.40 |
| maleic anhydride | 0.00 | 0.27 | 0.65 | 0.35 |
| s-acetylmercapto succinic anhydride | 0.00 | 0.30 | 0.48 | 0.38 |
| 2-octadecen-1-yl succinic anhydride | 0.00 | 0.28 | 0.55 | 0.35 |
| 18-crown-6 | 0.00 | 0.30 | 0.60 | 0.35 |
| benzo-18 crown-6 | 0.16 | 0.41 | 1.00 | 0.60 |
| dibenzo-18 crown-6 | 0.60 | 0.60 | 1.20 | 0.65 |
| dibenzo-24 crown-8 | 0.00 | 0.30 | 1.00 | 0.50 |
| 5-amino-3-methyl isooxazole | 0.00 | 0.32 | 0.55 | 0.45 |
| 2-oxazolidone | 0.50 | 0.71 | 0.95 | 0.75 |
| 5,5-dimethyl oxazolidine-2,4-dione | 0.15 | 0.37 | 0.90 | 0.44 |
| 3-ethyl-2-thioxo-4-oxazolidinone | 0.00 | 0.22 | 0.45 | 0.35 |
| 3-morpholino-1,2-propandiol | 0.20 | 0.35 | 0.73 | 0.55 |
| 4-phenyl morpholine | 0.00 | 0.30 | 0.55 | 0.32 |
| *N,N'* -dibenzyl-1,4,10,13-tetraoxa-7,16 diazacycloocta-decane | 0.00 | 0.26 | 0.70 | 0.30 |
| 4,7,13,16,21,24-hexaoxa-1,10-diazabicyclo [8.8.8] hexacosane | 0.00 | 0.30 | 0.70 | 0.60 |
| γ-valerolactam | 0.20 | 0.46 | 1.15 | 0.51 |
| ε-caprolactam | 0.00 | 0.26 | 0.50 | 0.35 |
| 2-azacyclooctanone | 0.00 | 0.30 | 0.45 | 0.40 |
| 2-azacyclononanone | 0.00 | 0.30 | 0.41 | 0.40 |
| maleimide | 0.00 | 0.35 | 0.70 | 0.35 |
| n-methylsuccinimide | 0.00 | 0.32 | 0.70 | 0.42 |
| phthalimide DBU salt | 0.00 | 1.20 | 0.20 | 0.80 |
| 1-allyl-2-thiourea | 0.00 | 0.52 | 1.00 | 0.55 |
| 1-benzyl-3-methyl-2-thiourea | 0.00 | 0.22 | 1.12 | 0.33 |
| 2-imino-4-thiobiuret | 0.00 | 0.60 | 1.25 | 0.67 |
| butyl sulfone | 0.00 | 0.25 | 0.72 | 0.40 |
| 2,2'-bithiophene | 0.00 | 0.58 | 1.45 | 0.58 |
| 2-phenyl-1,3-dithiane | 0.00 | 0.30 | 0.50 | 0.41 |
| 3,6,9,14-tetrathiabicyclo [9.2.1] tetradeca-11,13-diene | 0.25 | 0.50 | 1.10 | 0.65 |
| 1,5,9,13-tetra-thiacyclohexadecane-3,11-diol | 0.00 | 0.30 | 0.60 | 0.45 |
| 1,4,7,10,13-penta-thiacyclopentadecane | 0.60 | 0.70 | 1.50 | 0.70 |
| 2-aminothiazole | 0.10 | 0.30 | 1.60 | 0.45 |
| 2-amino-2-thiazoline | 0.00 | 0.23 | 0.65 | 0.30 |
| 3-methyl rhodanine | 0.20 | 0.50 | 1.85 | 0.33 |
| 3-ethyl-5-(2-hydroxy-ethyl)-4- methylthiazolium bromide | 0.00 | 0.29 | 1.04 | 0.32 |
| triphenylphosphine | 0.00 | 0.28 | 0.55 | 0.32 |
| tricyclohexylphosphine | 0.20 | 0.25 | 0.68 | 0.35 |
| 1,3-bis (diphenylphosphino) propane | 0.00 | 0.22 | 0.76 | 0.31 |
| 1,5-his(diphenyl phosphino) pentane | 0.00 | 0.23 | 0.48 | 0.30 |
| isopropyldiphenyl phosphine | 0.10 | 0.23 | 0.55 | 0.30 |
| triethyl phosphite | 0.00 | 0.25 | 0.70 | 0.33 |
| triphenyl phosphite | 0.00 | 0.05 | 0.30 | 0.05 |
| triethyl phosphite copper iodide | 0.20 | 0.28 | 0.46 | 0.25 |
| dipropyl phosphite | 0.00 | 0.05 | 0.12 | 0.05 |
| bis(2-ethylhexyl) phosphite | 0.00 | 0.15 | 0.70 | 0.12 |
| bis(4-nitrobenzyl) phosphite | 0.10 | 0.20 | 1.15 | 0.15 |
| diphenyl phosphine oxide | 0.00 | 0.23 | 0.66 | 0.31 |
| diphenyl(2,4,6-trimethylbenzoyl) phosphine oxide | 0.00 | 0.26 | 3.45 | 0.31 |
| vinyl phosphonic acid | 0.00 | 0.24 | 0.65 | 0.30 |
| cyanoaceto-hydrazide | 0.10 | 0.35 | 0.95 | 0.45 |
| cyanomethyl *N,N*-dimethyl dithiocarbamate | 0.00 | 0.56 | 1.00 | 0.40 |
| 4'-pentyl-4'-biphenyl carbonitrile | 0.00 | 0.22 | 1.15 | 0.30 |
| 4'-(octyloxy)-4-biphenyl carbonitrile | 0.00 | 0.30 | 0.70 | 0.39 |
| 1,4-dicyano-2-butene | 0.00 | 0.30 | 0.68 | 0.40 |
| benzylidene malononitrile | 0.00 | 0.30 | 1.00 | 0.35 |
| 1-isothiocyanato-4-(*trans*-4-propylcyclohexyl)benzene | 0.00 | 0.33 | 0.70 | 0.35 |
| formamidoxime | 0.00 | 0.28 | 1.00 | 0.35 |
| ethyl chlorooximido acetate | 0.00 | 0.09 | 0.15 | 0.07 |
| acetohydroxamic acid | 0.00 | 0.25 | 0.50 | 0.35 |
| tetraheptylammonium chloride | 0.00 | 0.25 | 0.80 | 0.32 |
| tetraheptylammonium bromide | 0.00 | 0.30 | 0.75 | 0.30 |

As the data indicate, contact between the migration marking material and the indicated transparentizing agents while the softenable material was in a molten state resulted in transparentization of the migration marking material. The process was repeated except that poly (2-hydroxyethyl methacrylate) (obtained from Scientific Polymer Products, #414) was substituted for the styrene/ethyl acrylate/acrylic acid terpolymer as the binder. Substantially similar results were obtained.

### EXAMPLE II

Migration imaging members were prepared as described in Example I. The surfaces of the members thus formed were uniformly negatively charged to a surface potential of -142 Volts with a corona charging device and were subsequently optically exposed by placing test pattern masks comprising silver halide images in contact with the imaging members and exposing the members to blue light of 480 nanometers through the mask for a period of 5 seconds. The imaging members were then developed by heating them with an aluminum heating block in contact with the polyester substrates at temperatures of from about 85 to about 100°C for about 5 seconds. Images corresponding to the images on the test pattern masks were subsequently visible in the developed imaging members.

The developed migration imaging members were then cut into pieces and pieces containing only Dmin areas (i.e., areas wherein the selenium particles had migrated in depth through the softenable layer) were placed in intimate contact with polyester sheets coated with a binder and a transparentizing agent and prepared as described in Example I. The UV absorption spectra at 685 nm of the Dₘᵢₙ areas of the migration imaging members were measured to determine the extent of migration marking material transparentization. UV absorption spectra were measured with a Shimadzu UV-160 spectrometer; all spectra were recorded by using 50% transmission aluminized ICI 442 polyester as a reference. The optical densities of the Dₘᵢₙ areas of the migration imaging members were also measured with a Macbeth TR927 densitometer in the visible, ultraviolet, and infrared range, using a Wratten No. 47 filter for the blue measurements, a Wratten No. 18A filter for the UV measurements, and a Wratten No. 25 filter for the IR measurements. For comparison purposes, the UV absorption spectrum at 685 nm and the optical density of the Dₘᵢₙ areas of the migration imaging members prior to contact with the sheet coated with transparentizing agent were also measured. The results were as follows:

| Agent | UV absorption | Optical Density | | |
|---|---|---|---|---|
| | | vis. | UV | IR |
| none | 1.45 | 0.74 | 1.63 | 0.79 |
| piperidine | 0.00 | 0.25 | 0.85 | 0.35 |
| 2-piperidine methanol | 0.50 | 0.50 | 0.40 | 0.28 |
| bis(pentamethylene) urea | 0.00 | 0.25 | 0.50 | 0.30 |
| 4,4'-trimethylene bis(1-piperidine propionitrile) | 0.00 | 0.20 | 0.50 | 0.40 |
| homopiperazine | 0.00 | 0.25 | 0.50 | 0.28 |
| hexacyclentrisulfate | 0.25 | 0.40 | 0.80 | 0.50 |
| 5,10,15,20-tetraphenyl-21H,23Hporphine | 0.25 | 0.50 | 0.78 | 0.50 |
| 3-pyrrolidino-1,2-propanediol | 0.00 | 0.24 | 0.75 | 0.28 |
| 1-dodecyl pyridinium chloride | 0.00 | 0.29 | 0.80 | 0.30 |
| 7,8-benzoquinoline | 0.15 | 0.28 | 0.61 | 0.33 |
| 8-hydroxyquinaldine | 0.05 | 0.26 | 0.74 | 0.35 |
| phthalazine | 0.25 | 0.30 | 0.85 | 0.36 |
| 1,10-phenanthroline | 0.10 | 0.36 | 0.80 | 0.42 |
| 1,3,5-triazine | 0.00 | 0.42 | 0.83 | 0.40 |
| norbornane | 0.05 | 0.30 | 0.80 | 0.45 |
| γ-butyrolactone | 0.00 | 0.45 | 1.01 | 0.52 |
| 1,3,5-trioxane | 0.00 | 0.28 | 0.66 | 0.31 |
| piperonal | 0.00 | 0.29 | 0.65 | 0.35 |
| piperonylalcohol | 0.00 | 0.23 | 0.55 | 0.37 |
| maleic anhydride | 0.00 | 0.28 | 0.73 | 0.34 |
| benzo-18-crown-6 | 0.10 | 0.35 | 0.77 | 0.33 |
| 5-amino-3-methyl isooxazole | 0.00 | 0.28 | 0.57 | 0.40 |
| 3-ethyl-2-thioxo-4-oxazolidinone | 0.00 | 0.26 | 0.85 | 0.31 |
| 3-morpholino-1,2-propandiol | 0.10 | 0.37 | 0.88 | 0.42 |
| 4-phenyl morpholine | 0.00 | 0.26 | 0.65 | 0.32 |
| *N,N'*-dibenzyl-1,4,10,13-tetraoxa-7,16 diazacyclooctadecane | 0.00 | 0.24 | 0.65 | 0.30 |
| γ-valerolactam | 0.10 | 0.29 | 0.83 | 0.31 |
| 2-azacyclooctanone | 0.00 | 0.26 | 0.74 | 0.38 |
| 1-allyl-2-thiourea | 0.00 | 0.30 | 0.95 | 0.35 |
| 1,3-dithiane | 0.15 | 0.34 | 0.54 | 0.35 |
| 2-amino-2-thiazoline | 0.00 | 0.23 | 0.90 | 0.30 |
| 3-ethyl-5-(2-hydroxy-ethyl)-4-methylthiazolium bromide | 0.00 | 0.31 | 1.09 | 0.27 |
| triphenylphosphine | 0.00 | 0.31 | 0.87 | 0.29 |
| tricyclohexylphosphine | 0.10 | 0.30 | 0.75 | 0.40 |
| 1,3-bis(diphenyl-phosphino) propane | 0.00 | 0.25 | 0.80 | 0.35 |
| 1,5-bis(diphenyl phosphino) pentane | 0.00 | 0.26 | 0.60 | 0.30 |
| triethyl phosphite copper iodide | 0.10 | 0.35 | 0.50 | 0.33 |
| bis(4-nitrobenzyl) phosphite | 0.10 | 0.25 | 0.80 | 0.30 |
| diphenyl phosphine oxide | 0.00 | 0.24 | 0.71 | 0.35 |
| vinyl phosphonic acid | 0.00 | 0.30 | 0.75 | 0.25 |
| triphenyl phosphate | 0.20 | 0.35 | 0.80 | 0.45 |
| cyanoaceto-hydrazide | 0.10 | 0.30 | 0.92 | 0.42 |
| 1-isothiocyanato-4-(*trans*-4-propylcyclohexyl)benzene | 0.00 | 0.41 | 0.72 | 0.41 |
| formamidoxime | 0.00 | 0.28 | 1.30 | 0.38 |
| acetohydroxamic acid | 0.00 | 0.23 | 0.77 | 0.30 |
| tetrahexylammonium chloride | 0.40 | 0.34 | 0.90 | 0.41 |
| tetraheptylammonium bromide | 0.00 | 0.27 | 0.75 | 0.30 |

As the data indicate, contact between the migration marking material in the Dₘᵢₙ areas and the indicated transparentizing agents while the softenable material was in a molten state resulted in transparentization of the migration marking material in the Dₘᵢₙ areas. The process was repeated except that poly (2-hydroxyethyl methacrylate) (obtained from Scientific Polymer Products, #414) was substituted for the styrene/ethyl acrylate/acrylic acid terpolymer as the binder. Substantially similar results were obtained.

### EXAMPLE III

Migration imaging members are prepared as described in Example I with the exception that prior to coating the softenable layer onto the polyester substrate, the polyester substrate is first coated as follows. A solution is prepared of toluene containing about 10 percent solids, wherein the solids comprise about 10 percent by weight of a transparentizing agent and about 90 percent by weight of a styrene/ethyl acrylate/acrylic acid terpolymer. The resulting solution is coated by a solvent extrusion technique onto the polyester substrates. The layer thus deposited is allowed to dry at about 25°C for about 1 hour, resulting in a dried transparentizing layer with a thickness of about 2 microns. Thereafter, the softenable layer is coated onto the transparentizing layer by the method described in Example I. The transparentizing agents used are those set forth in Examples I and II. During the selenium vacuum deposition process, the transparentizing layer and the softenable layer fuse to form a single softenable layer with the transparentizing agent concentrated in the bottom area thereof. The imaging members thus formed are imaged as described in Example II. It is believed that the optical contrast density of these imaging members will be greater than that of an imaging member of identical composition except that it contains no transparentizing agent, and that the optical density of the Dₘᵢₙ areas of these imaging members will be less than that of an imaging member of identical composition except that it contains no transparentizing agent.

### EXAMPLE IV

Migration imaging members are prepared as described in Example I with the exception that the solution for the softenable layer is prepared by dissolving about 76 parts by weight of the styrene/ethyl acrylate/acrylic acid terpolymer, about 14 parts by weight of the charge transporting compound, and about 10 parts by weight of a transparentizing agent. The transparentizing agents used are those set forth in Examples I and II. The imaging members thus formed are imaged as described in Example II. It is believed that the optical contrast density of these imaging members will be greater than that of an imaging member of identical composition except that it contains no transparentizing agent, and that the optical density of the Dₘᵢₙ areas of these imaging members will be less than that of an imaging member of identical composition except that it contains no transparentizing agent.

### EXAMPLE V

Migration imaging members are prepared as described in Example I with the exception that prior to coating the softenable layer onto the polyester substrate, the polyester substrate is first coated as follows. A solution is prepared of methanol containing about 10 percent solids, wherein the solids comprise about 10 percent by weight of a transparentizing agent and about 90 percent by weight of a poly (2-hydroxyethyl methacrylate) binder (available from Scientific Polymer Products). The resulting solution is coated by a solvent extrusion technique onto the polyester substrates. The layer thus deposited is allowed to dry at about 25°C for about 1 hour, resulting in a dried transparentizing layer with a thickness of about 2 microns. Thereafter, the softenable layer is coated onto the transparentizing layer by the method described in Example I. The transparentizing agents used are those set forth in Examples I and II. The imaging members thus formed are imaged as described in Example II. It is believed that the optical contrast density of these imaging members will be greater than that of an imaging member of identical composition except that it contains no transparentizing agent, and that the optical density of the Dₘᵢₙ areas of these imaging members will be less than that of an imaging member of identical composition except that it contains no transparentizing agent.

### EXAMPLE VI

Migration imaging members are prepared as described in Example I with the exception that subsequent to vacuum deposition of the selenium migration marking material, the softenable layer is coated as follows. A solution is prepared of methanol containing 10 percent by weight solids, wherein the solids comprise about 10 percent by weight of a transparentizing agent and about 90 percent by weight of a poly (2-hydroxyethyl methacrylate) binder. The resulting solution is coated by a solvent extrusion technique onto the softenable layers containing migration marking material. The layer thus deposited is allowed to dry at about 25°C for about 1 hour, resulting in a dried transparentizing layer with a thickness of about 2 microns. The transparentizing agents used are those set forth in Examples I and II. The imaging members thus formed are imaged as described in Example II. It is believed that the optical contrast density of these imaging members will be greater than that of an imaging member of identical composition except that it contains no transparentizing agent, and that the optical density of the Dₘᵢₙ areas of these imaging members will be less than that of an imaging member of identical composition except that it contains no transparentizing agent.

## Claims

1. A migration imaging member (1) comprising (a) a substrate (2), (b) a softenable layer (6) comprising a softenable material (7) and a photosensitive migration marking material (8), and (c) a transparentizing agent which transparentizes the migration marking material in contact therewith contained in at least one layer of the migration imaging member, wherein the transparentizing agent affects the migration marking material which comes into contact therewith by reducing the optical density of the softenable layer containing the migration marking material.

2. A migration imaging member according to claim 1, wherein the migration marking material (8) is selected from the group consisting of (a) selenium, (b) tellurium, (c) alloys of selenium and a material selected from the group consisting of tellurium, arsenic, antimony, thallium, bismuth, or mixtures thereof, (d) alloys of tellurium and a material selected from the group consisting of arsenic, antimony, thallium, bismuth, or mixtures thereof, (e) halogen doped selenium, (f) halogen doped tellurium, (g) halogen doped alloys of selenium and a material selected from the group consisting of tellurium, arsenic, antimony, thallium, bismuth, or mixtures thereof, (h) halogen doped alloys of tellurium and a material selected from the group consisting of arsenic, antimony, thallium, bismuth, or mixtures thereof, and (i) mixtures thereof.

3. A migration imaging member according to claim 1 or claim 2, wherein the transparentizing agent is contained in the softenable layer.

4. A migration imaging member according to claim 1 or claim 2, wherein the transparentizing agent is contained in a layer situated between the softenable layer and the substrate.

5. The migration imaging member according to claim 1 or 2, wherein the softenable layer is situated between the substrate and a layer containing the transparentizing agent.

6. A migration imaging member according to claim 1 or claim 2, wherein the migration imaging member comprises a substrate, a first softenable layer comprising a first softenable material and a first migration marking material, and a second softenable layer comprising a second softenable material and a second migration marking material, wherein the transparentizing agent is contained in a layer situated between the first softenable layer and the second softenable layer.

7. A migration imaging member according to any of claims 1 to 6, wherein the transparentizing agent is present in an amount of from about 1 to about 50 percent by weight of the material comprising the layer in which it is contained.

8. A migration imaging member according to claim 1 wherein the transparentizing agent is an azacyclic compound; or wherein the transparentizing agent is selected from the group consisting of: (A) materials of the general formulae: wherein R₁, R₂, R₃, R₄, R₅, R₆, R₇, R₈, R₉, R₁₀, R₁₁, R₁₂, R₁₃, R₁₄, Rᵢₛ, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈, and R₃₉ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈, and R₃₉ can be joined together to form a ring; (B) materials of the general formulae: wherein R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, and R₂₂ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, and R₂₂ can be joined together to form a ring; (C) materials of the general formulae: wherein R₁, R₂, and R₃ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, and R₃ can be joined together to form a ring; (D) materials of the general formulae: wherein R₁, R₂, R₃, R₄, R₅, R₆, R₇, R₈, R₉, R₁₀, R₁₁, and R₁₂ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, and R₁₂ can be joined together to form a ring; (E) materials of the general formulae: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (F) materials of the general formula: R₁, R₂, R₃, R₄, R₅, R₆, R₇, R₈, R₉, R₁₀, R₁₁, R₁₂, R₁₃, and R₁₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, and R₁₄ can be joined together to form a ring; (G) materials of the general formula: wherein R₁ and R₂ each, independently of the other, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein R₁ and R₂ can be joined together to form a ring; (H) materials of the general formula: wherein R₁, R₂, R₃, R₄, and R₅ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, and R₅ can be joined together to form a ring; (I) materials of the general formula: wherein R₁, R₂, R₃, R₄, R₅, R₆, R₇, R₈, and R₉ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, and R₉ can be joined together to form a ring; (J) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (K) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (L) materials of the general formula: wherein R₁, R₂, R₃, R₄, and R₅ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, and R₅ can be joined together to form a ring; (M) materials of the general formulae: wherein R₁, R₂, R₃, R₄, R₅, R₆, R₇, R₈, R₉, R₁₀, R₁₁, R₁₂, R₁₃, and R₁₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, and R₁₄ can be joined together to form a ring; (N) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (O) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (P) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (Q) materials of the general formula: wherein R₁, R₂, R₃, and R₄ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, and R₄ can be joined together to form a ring; (R) materials of the general formulae: wherein R₁ is selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, and wherein the curved portion of the structure represents a hydrocarbon chain or a substituted hydrocarbon chain, wherein two or more substituents can be joined together to form a ring; (S) materials of the general formula: wherein R₁ is selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, and wherein the curved portion of the structure represents a hydrocarbon chain or a substituted hydrocarbon chain, wherein two or more substituents can be joined together to form a ring; and (T) mixtures thereof; or wherein the transparentizing agent is selected from the group consisting of (1) homopiperidine, (2) piperidinethiocyanate, (3) -2-piperidinemethanol, (4) 3-piperidinemethanol, (5) 2-piperidineethanol, (6) 4-piperidineethanol, (7) 4-piperidine monohydrate hydrochloride, (8) 1-aminopiperidine, (9) 1-(2-aminoethyl)piperidine, (10) 4-(aminomethyl)piperidine, (11) 3-piperidino-1,2-propanediol (Aldrich 21,849-9), (12) 1-piperidine propionic acid, (13) 1-methyl-4-(methylamino)piperidine, (14) 1-acetyl-3-methylpiperidine, (15) 4'-piperidinoacetophenone, (16) 4-phenylpiperidine, (17) 4-piperidinopiperidine, (18) 4-benzylpiperidine, (19) 4-(4-methylpiperidino)pyridine, (20) 4-piperidone ethylene ketal, (21) bis(pentamethylene)urea, (22) 1-benzyl-4-hydroxypiperidine, (23) 1-benzoyl-4-piperidone, (24) 1,1'-methylenebis(3-methylpiperidine), (25) 4,4'-trimethylenedipiperidine, (26) 4,4'-trimethylenebis(1-menthylpiperidine), (27) 4,4'-trimethylenebis(1-piperidinepropionitrile), (28) 4,4'-trimethylenebis(1-piperidineethanol), (29) 2,2,6,6-tetramethylpiperidine, (30) 4-amino-2,2,6,6-tetramethylpiperidine, (31) 4-(dimethylamino)-1,2,2,6,6-pentamethylpiperidine, (32) N,N'-bis(2,2,6,6-tetramethyl-4-piperidinyl)-1,6-hexanediamine, (33) tripiperidinophosphine oxide, (34) tropane, (35) tropinehydrate, (36) tropinone, (37) 8-hydroxytropinone, (38) 2-piperidine carboxylic acid, (39) 2-piperidone, (40) 4,4'-trimethylene bis (1-piperidine carboxamide), (41) 4-methyl-2-(piperidinomethyl) phenol, (42) 1-methyl-4-piperidinyl bis (chlorophenoxy) acetate, (43) 2-(hexamethylene imino) ethyl chloride monohydrochloride, (44) 3-(hexahydro-1H-azepin-1-yl)-3'-nitropropiophenone hydrochloride, (45) imipramine hydrochloride, (46) carbamezepine, (47) 5,6,11,12-tetrahydro dibenz [b,f] azocine hydrochloride, (48) quinuclidine hydrochloride, (49) 3-quinuclidinol hydrochloride, (50) 3-quinuclidinone hydrochloride, (51) 2-methylene-3-quinuclidinone dihydrate hydrochloride, (52) 3-amino quinuclidine dihydrochloride, (53) 3-chloro quinuclidine hydrochloride, (54) quinidine sulfate dihydrate, (55) quinine monohydrochloride dihydrate, (56) quinine sulfate monohydrate, (57) hydroquinidine hydrochloride, (58) hydroquinine hydrobromide dihydrate, (59) piperazine, (60) homopiperazine, (61) 1-methylpiperazine, (62) 2-methylpiperazine, (63) 1-acetylpiperazine, (64) 1-(2-hydroxyethyl)piperazine, (65) 1-(2-aminoethyl)piperazine, (66) tert-butyl 1-piperazinecarboxylate, (67) N-isopropyl-1-piperazineacetamide, (68) 1-(2-methoxyphenyl)piperazine, (69) 1-(2-pyridyl)piperazine, (70) 1-benzylpiperazine, (71) 1-cinnamylpiperazine, (72) 1-(4-chlorobenzhydryl)piperazine, (73) 2,6-dimethylpiperazine, (74) 1-amino-4-methylpiperazine, (75) 1-amino-4-(2-hydroxyethyl)piperazine, (76) 1,4-bis(2-hydroxyethyl)piperazine, (77) 1,4-bis(3-aminopropyl)piperazine, (78) tert-butyl-4-benzyl-1-piperazinecarboxylate, (79) 1-piperonyl piperazine, (80) bis(4-methyl-1-homopiperazinylthiocarbonyl)disulfide, (81) 1-amino-4-methyl piperazine dihydrochloride monohydrate, (82) 1-(3-chloropropyl)-piperazine dihydrochloride monohydrate, (83) 1-(2,3-xylyl) piperazine monohydrochloride, (84) 1,1-dimethyl-4-phenyl piperazineium iodide, (85) 1,4,7-triazacyclononane, (86) 1,5,9-triazacyclododecane, (87) 1,2,3-triazole, (88) 4-amino-1,2,4-triazole, (89) 3-amino-5-methylthio-lH-1,2,4-triazole, (90) benzotriazole, (91) 1-aminobenzotriazole, (92) 1-cyanobenzotriazole, (93) 5-methyl-1H-benzotriazole, (94) 1H-benzotriazole-1-ylmethyl isocyanide, (95) 2-[3-(2H-benzotriazole-2-yl)-4-hydroxyphenyl]ethyl methacrylate, (96) 1,2,4-triazole, (97) 1,2,4-triazole sodium derivative, (98) 3-amino-1,2,4-triazole, (99) 3,5-diamino-1,2,4-triazole, (100) 3-amino-5-mercapto-1,2,4-triazole, (101) 3-amino-1,2,4-triazole-5-carboxylic acid hemihydrate, (102) 4-amino-3-hydrazino-5-mercapto-1,2,4-triazole, (103) 1,2,3-triazole-4,5-dicarboxylic acid monohydrate, (104) nitron, (105) 1-hydroxybenzotriazole hydrate, (106) 1,3,5-triazine, (107) cyanuric acid, (108) trithiocyanuric acid, (109) 2,4-bis (methylthio)-6-chloro-1,3,5-triazine, (110) 2-chloro-4,6-dimethoxy-1,3,5-triazine, (111) 2-chloro-4,6-diamino-1,3,5-triazine, (112) trichloromelamine, (113) cyanuric chloride, (114) 2,4,6-tris(perfluoroheptyl)-1,3,5-triazine, (115) hexahydro-2,4,6-trimethyl-1,3,5-triazine trihydrate, (116) 1,3,5-trimethylhexahydro-1,3,5-triazine, (117) 1,3,5-triethylhexahydro-1,3,5-triazine, (118) 1,3,5-triclohexylhexahydro-1,3,5-triazine, (119) 1,3,5-tribenzylhexahydro-1,3,5-triazine, (120) trichloroisocyanuric acid, (121) tris (2,3-dibromopropylisocyanurate), (122) cyanuric acid compound with melamine, (123) urazole, (124) 1-methyl urazole, (125) 4-phenyl urazole, (126) 5-(4-hydroxyphenyl)-5-phenyl hydantoin, (127) β-tetralone hydantoin, (128) cyclen (1,4,7,10-tetraazacyclododecane), (129) 1,4,8,11-tetraazacyclotetradecane, (130) 1,4,8,11-tetramethyl-1,4,8,11-tetraazacydotetradecane, (131) 1,4,8,11-tetraazacyclotetradecane-5,7-dione, -dione, (132) 1,4,8,12-tetraazacyclopentadecane, (133) 2,3,7,8,12,13,17,18-octaethyl-21H,23H-porphine, (134) dimethyl 3,7,12,17-tetramethyl-21H,23H-porphine-2,18-dipropionate, (135) dimethyl 7,12-diacetyl-3,8,13,17-tetramethyl-21H,23H-porphine-2,18-dipropionate, (136) 8,3-divinyl-3,7,12,17-tetramethyl-21H,23H-porphine-2,18-dipropionic acid, disodium salt, (137) 5,10,1 5,20-tetraphenyl-21 H,23H-porphine, (138) 5,10,15,20-tetrakis(4-methoxyphenyl)-21H,23H-porphine, (139) 5,10,15-20-tetrakis[4-(trimethylamino)phenyl]-21H,23H-porphine tetra-p-tosylate salt, (140) 5,10,15,20-tetra(4-pyridyl)-21H,23H-porphine, (141) 5,10,15,20-tetrakis(1-methyl-4-pyridyl)-21H,23H-porphine, tetra-p-tosylate salt), (142) 1,5-pentamethylenetetrazole, (143) 1-H-tetrazole, (144) 5-amino tetrazole monohydrate, (145) 2,3,5-triphenyl-2H-tetrazolium chloride, (146) 2-(4-iodophenyl)-5-(4-nitrophenyl)-3-phenyltetrazolium chloride, (147) 1,2,3,3-tetramethyl-3H-indolinium iodide, (148) hexacyclen trisulfate, (149) hexamethylhexacyclen, (150) pyrrole-2-carboxaldehyde, (151) proline amide, (152) 3-pyrrolidino-1,2-propane diol, (153) 1-(pyrrolidino carbonylmethyl) piperazine, (154) 4-pyrrolidinopyridine, (155) 3-indolylacetonitrile, (156) 6-nitroindoline, (157) 7-azaindole, (158) indazole, (159) 2-acetyl-pyrrole, (160) 2-acetyl-1-methylpyrrole, (161) 3-acetyl-1-methylpyrrole, (162) 3-acetyl-2,4-dimethylpyrrole, (163) pyrrole-2-carboxylic acid, (164) 3-carboxy-1,4-dimethyl-2-pyrroleacetic acid, (165) proline, (166) 2-pyrrolidone-5-carboxylic acid, (167) 4-hydroxyproline, (168) 1,1'-ethylene bis (5-oxo-3-pyrrolidine carboxylic acid), (169) kainic acid monohydrate, (170) 1-amino pyrrolidine hydrochloride, (171) 2-(2-chloroethyl)-1-methyl pyrrolidine hydrochloride, (172) 1-(2-chloroethyl) pyrrolidine hydrochloride, (173) tremorine dihydrochloride, (174) L-proline methyl ester hydrochloride, (175) ammonium pyrrolidine dithiocarbamate, (176) pyrrolidone hydrotribromide, (177) 1-(4-chlorobenzyl)-2-(1-pyrrolidinyl methyl) benzimidazole hydrochloride, (178) billverdin dihydrochloride, (179) indole, (180) 4,5,6,7-tetrahydroindole, (181) 3-indolemethanol hydrate, (182) 3-indole ethanol, (183) indole-3-carboxaldehyde, (184) 3-indolylacetate, (185) indole-3-acetamide, (186) indole-3-carboxylic acid, (187) indole-3-acetic acid, (188) 3-indole propionic acid, (189) 3-indole acrylic acid, (190) 3-indole glyoxylic acid, (191) indole-3-pyruvic acid, (192) 3-indolelactic acid, (193) 3-indole butyric acid, (194) N-acetyltryptophanamide, (195) N-(3-indolylacetyl)alanine, (196) N-(3-indolyl acetyl)valine, (197) N-(3-indolyl acetyl)isoleucine, (198) N-(3-indolyl acetyl)leucine, (199) N-(3-indolyl acetyl)aspartic acid, (200) N-(3-indolyl acetyl)-L-phenylalanine, (201) 4-hydroxyindole, (202) indole-4-carboxylic acid, (203) 4-indolyl acetate, (204) 4-methyl indole, (205) 5-hydroxy indole, (206) 5-hydroxy indole-3-acetic acid, (207) 5-hydroxy-2-indole carboxylic acid, (208) N-acetyl-5-hydroxytryptamine, (209) indole-5-carboxylic acid, (210) 5-methyl indole, (211) 5-methoxy indole, (212) indole-2-carboxylic acid, (213) indolene-2-carboxylic acid, (214) indole-2,3-dione, (215) 2-methyl indole, (216) 2,3,3-trimethyl indolenine, (217) tryptamine hydrochloride, (218) 5-methyl tryptamine hydrochloride (219) serotonin hydrochloride hemihydrate, (220) norharman hydrochloride monohydrate, (221) harmane hydrochloride monohydrate, (222) harmine hydrochloride hydrate, (223) harmaline hydrochloride dihydrate, (224) harmol hydrochloride dihydrate, (225) harmalol hydrochloride dihydrate, (226) 3,6-diamino acridine hydrochloride, (227) (3-indolyl) isothiuronium iodide, (228) yohimbine hydrochloride, 229) pyrazole, (230) 3-amino pyrazole, (231) 5-amino-1-ethylpyrazole, (232) 3-amino-4-carbethoxypyrazole, (233) 3-amino-5-methylpyrazole, (234) 3-amino-5-phenylpyrazole, (235) ethyl 4-pyrazole carboxylate, (236) diethyl 3,5-pyrazolecarboxylate, (237) 1,1'-(1-ethylpropylidene)bis 1H-pyrazole, (238) 4-bromopyrazole, (239) 4-bromo-3-methyl pyrazole, (240) 3,5-dimethyl pyrazole, (241) 4-bromo-3,5-dimethyl pyrazole, (242) 3,5-dimethyl pyrazole-1-carboxamide, (243) 3,5-dimethylpyrazole-1-methanol, (244) 3-methyl-1-vinylpyrazole, (245) 4-benzoyl-3-methyl-1-phenyl-2-pyrazolin-5-one, (246) 1-nitropyrazole, (247) 4-pyrazole carboxylic acid, (248) 3,5-pyrazole dicarboxylic acid monohydrate, (249) 3-amino-5-hydroxypyrazole, (250) 3-amino-4-pyrazole carbonitrile, (251) 3-amino-4-pyrzaolecarboxylic acid, (252) 4-methyl pyrazole hydrochloride, (253) 3,4-diamino-5-hydroxy pyrazole sulfate, (254) (3,5-dimethyl pyrazole-1-carboxamidine nitrate), (255) 3-amino-4-pyrazole carboxamide hemisulfate, (256) acid salt of 6-amino indazole hydrochloride, (257) 4-hydroxypyrazolo [3,4-d] pyrimidine, (258) 4-mercapto-1H-pyrazolo-[3,4-d]-pyrimidine, (259) indazole, (260) 5-aminoindazole, (261) 6-aminoindazole, (262) 3-indazolinone, (263) N'-(6-indazolyl) sulfanilamide, (264) 4,5-dihydro-3-(4-pyridinyl)-2H-benz[g] indazole methane sulfonate, (265) imidazole, (266) 4-methylimidazole, (267) 2-ethylimidazole, (268) 2-propylimidazole, (269) 1-butylimidazole, (270) 2-undecylimidazole, (271) histamine, (272) 1-(3-aminopropyl) imidazole, (273) 1-acetylimidazole, (274) 2-methyl-1-vinylimidazole, (275) 2-ethyl-4-methylimidazole, (276) 1-benzyl-2-methylimidazole, (277) 1-methylbenzimidazole, (278) 1-ethyl-3-methyl-1,H-imidazolinium chloride, (279) 2-(aminomethyl) benzimidazole dihydrochloride hydrate, (280) 2,6-diamino-8-purinol hemisulfate monohydrate, (281) purin-6-yl-trimethyl ammonium chloride, (282) 4-methyl-5-imidazole methanol hydrochloride, (283) N,N'-bis[3-(4,5-dihydro-1H-imidazol-2-yl)phenyl]urea dipropanoate, (284) 1-(p-tosyl)-3,4,4-trimethyl-2-imidazolinium iodide, (285) 1-ethyl-3-methyl-1H-imidazolinium chloride, (286) 2-amino imidazole sulfate, (287) 4-amino-5-imidazole carboxamide hydrochloride, (288) 2-hydrazino-2-imidazoline hydrobromide, (289) imidazole hydrochloride, (290) 4-imidazole acetic acid hydrochloride, (291) 2-benzyl-2-imidazoline hydrochloride, (292) propyl-1-(1-phenyl ethyl imidazole-5-carboxylate hydrochloride, (293) 2,6-diamino purine sulfate hydrate, (294) 1-tallow amido ethyl-3-methyl-2-heptadecyl imidazolinium methyl sulfate, (295) isostearyl ethyl imidonium ethyl sulfate, (296) methyl-1-tallow amido ethyl-2-tallow imidazolinium methyl sulfate, (297) isostearyl benzyl imidonium chloride, (298) methyl-1-hydrogenated tallow amido ethyl (299) hydrogenated tallow imidazolinium methyl sulfate, (300) 1-methyl-1-oleyl amido ethyl-2-oleyl-imidazolinium methyl sulfate, (301) cocohydroxyethyl polyethyleneglycol imidazolinium chloride phosphate, (302) guanine, (303) guanosine hydrate, (304) xanthine, (305) 1-methylxanthine, (306) 3-methyl xanthine, (307) 3-isobutyl-1-methyl xanthine, (308) hypoxanthin, (309) xanthosine dihydrate, (310) 6-thioxanthene, (311) purine, (312) 6-amino purine, (313) 6-methoxy purine hemihydrate, (314) 6-mercaptopurine monohydrate, (315) 2-amino-6-chloropurine, (316) 2-amino-6,8-dihydroxy purine, (317) theophylline (3,7 dihydro-1,3-dimethyl-1H-purine-2,6-dione), (318) kinetin, (319) 1-methyl adenine, (320) 3-methyl adenine, (321) adenosine, (322) inosine, (323) 6-mercaptopurine riboside, (324) 6-amino purine hydrochloride hemihydrate, (325) 6-amino purine sulfate, (326) 2,6-diamino-8-purinol hemisulfate monohydrate, (327) benzimidazole, (328) 2-aminobenzimidazole, (329) 2-amino-5,6-dimethlybenzimidazole, (330) 5-benzimidazole carboxylic acid, (331) 2,4,5-trimethyl benzimidazole, (332) 2-guanidinobenzimidazole, (333) 2-hydroxybenzimidazole, (334) 4-(2-keto-1-benzimidazolinyl) piperidine, (335) 2-imidazolidine thione, (336) 2-imidazolidone, (337) hydantoin, (338) 1-methyl hydantoin, (339) creatinine, (340) 2-thiohydrantoin, (341) 5-hydantoin acetic acid, (342) 5-ureidohydantoin, (343) 5,5-dimethyl hydantoin, (344) 2-imidazolidone-4-carboxylic acid, (345) N,N-bis (2-hydroxyethyl) isonicotinamide, (346) 1,2-bis(4-pyridyl) ethylene, (347) 2-(2-piperidinoethyl) pyridine, (348) 1,2-bis (4-pyridyl)ethane, (349) 4,4'-trimethylene pyridine, (350) aldrithiol-2, (351) aldrithiol-4, (352) 1,3-bis (3-pyridylmethyl)-2-thiourea, (353) 2,2':6',2"-terpyridine, (354) 2-[N,N-bis(triflouromethylsulfonyl)amino]pyridine, (355) 2,3-pyridine dicarboxylic acid, (356) 2,4-pyridine dicarboxylic acid monohydrate, (357) 2,5-pyridine dicarboxylic acid, (358) 2,6-pyridine dicarboxylic acid, (359) 3,4-pyridine dicarboxylic acid, (360) 3,5-pyridine dicarboxylic acid, (361) 2,6-pyridine dicarboxaldehyde, (362) 3,4-pyridine carboxamide, (363) 3,4-pyridine carboximide, (364) 2,3-pyridine carboxylic anhydride, (365) 3,4-pyridine carboxylic anhydride, (366) 2,6-pyridine methanol, (367) 2-pyridine ethane sulfonic acid, (368) 4-pyridine ethane sulfonic acid, (369) 3-pyridine sulfonic acid, (370) pyridoxic acid, (371) trans-3-(3-pyridyl) acrylic acid, (372) 2-pyridyl hydroxymethane sulfonic acid, (373) 3-pyridyl hydroxymethane sulfonic acid, (374) 6-methyl-2,3-pyridine dicarboxylic acid, (375) isonicotinic acid, (376) pyridine hydrobromide, (377) pyridine hydrochloride, (378) 2-(chloromethyl) pyridine hydrochloride, (379) 2-pyridylacetic acid hydrochloride, (380) nicotinoyl chloride hydrochloride, (381) 2-hydrazinopyridine dihydrochloride, (382) 2-(2-methyl aminoethyl) pyridine dihydrochloride, (383) 1-methyl-1,2,3,6-tetrahydropyridine hydrochloride, (384) 2,6-dihydroxypyridine hydrochloride, (385) 3-hydroxy-2(hydroxymethyl) pyridine hydrochloride, (386) pyridoxine hydrochloride, (387) pyridoxal hydrochloride, (388) pyridoxal 5-phosphate monohydrate, (389) 3-amino-2,6-dimethoxy pyridine hydrochloride, (390) pyridoxamine dihydrochloride monohydrate, (391) iproniazid phosphate, (392) tripelennamine hydrochloride, (393) pyridinium bromide perbromide, (394) pyridinium 3-nitrobenzenesulfonate, (395) 1-ethyl-3-hydroxy pyridinium bromide, (396) 1-ethyl-4-(methoxy carbonyl) pyridinium iodide, (397) 1-heptyl-4-(4-pyridyl) pyridinium bromide, (398) 1-dodecyl pyridinium chloride, (399) 1-hexadecyl pyridinium chloride monohydrate, (400) 1-hexadecyl pyridinium bromide monohydrate, (401) 1-(carboxymethyl) pyridinium chloride, (402) 1-(carboxymethyl) pyridinium chloride hydrazide, (403) 1-(3-nitrobenzyloxymethyl) pyridinium chloride, (404) 1-(3-sulfopropyl) pyridinium hydroxide, (405) N-(lauroyl colamino formyl methyl) pyridinium chloride, (406) N-(stearoyl colamine formyl methyl) pyridinium chloride, (407) 2-chloro-1-methyl pyridinium iodide, (408) 2-pyridine aldoxime-1-methyl methane sulfonate, 2-pyridine aldoxime-1-methyl chloride, (409) 2-[4-(dimethyl amino) styryl]1-ethylpyridinium iodide, (410) 1-benzyl-3-hydroxy pyridinium chloride, (411) 1,4 dimethyl pyridinium iodide, (412) 1-ethyl-4-phenyl pyridinium iodide, (413) 4-phenyl-1-propyl pyridinium iodide, (414) 1-docosyl-4-(4 hydroxystyryl) pyridinium bromide, (415) 1,1'-dimethyl-4-4'-bipyridinium dichloride, (416) 1,1'-diethyl-4-4'-bipyridinium dibromide, (417) 1,1'-dibenzyl-4,4'-bipyridinium dichloride, (418) 1,1'-diheptyl-4,4'-bipyridinium dibromide, (419) 1,7-phenanthroline, (420) 1,10-phenanthroline, (421) 5-chloro-1,10-phenanthroline, (422) 4,5-dihydro-3-(4-pyridinyl)-2H-benz[g] indazole methane sulfonate, (423) 1,2,3,4-tetrahydro quinoline, (424) 6-ethoxy-1,2,3,4-tetrahydro-2,2,4-trimethyl quinoline, (425) 2-cyanoquinoline, (426) 1-cyanoisoquinoline, (427) 3-cyanoisoquinoline, (428) 3-amino quinoline, (429) 8-aminoquinoline, (430) 7,8-benzoquinoline, (431) 8-hydroxy quinoline, (432) 8-hydroxyquinoline, aluminium salt, (433) 8-hydroxyquinaldine, (434) 3,4,5,6,7,8-hexahydro 2 (1H)-quinolinone, (435) julolidine, (436) quinoxaline, (437) ethyl-2-quinoxalinecarboxylate, (438) quinoline, (439) 2-hydroxyquinoline, (440) 4-hydroxy quinoline, (441) 5-hydroxy quinoline, (442) 5-amino quinoline, (443) 6-amino quinoline, (444) 2-quinoline carboxylic acid, (445) 3-quinoline carboxylic acid, (446) 4-quinoline carboxylic acid, (447) 4-quinoline carboxaldehyde, (448) 2-quinoline thiol, (449) 2,4-quinoline diol, (450) quinaldine, (451) 4-aminoquinaldine, (452) 2,6-dimethyl quinoline, (453) 2,7-dimethyl quinoline, (454) 4-methoxy-2-quinoline carboxylic acid, (455) methyl-2-phenyl-4-quinoline carboxylate, (456) 2-(N-butyl carbamoyl)-1,2,3,4-tetrahydro-isoquinoline, (457) 1-hydroxyisoquinoline, (458) 1-isoquinoline carboxylic acid, (459) 3-isoquinoline carboxylic acid, (460) 1,5-isoquinoline diol, (461) 8-hydroxyquinoline hemisulfate hemihydrate, (462) 5-amino-8-hydroxy quinoline dihydrochloride, (463) 2-(chloromethyl) quinoline monohydrochloride, (464) 8-hydroxyquinoline-5-sulfonic acid monohydrate, (465) 8-ethoxy-5-quinoline sulfonic acid sodium salt hydrate, (466) 1,2,3,4-tetrahydroisoquinoline hydrochloride, (467) 1,2,3,4-tetrahydro-3-isoquinoline carboxylic acid hydrochloride, (468) 6,7-dimethoxy-1,2,3,4-tetrahydro isoquinoline hydrochloride, (469) 1-methyl-6,7-dihydroxy-1,2,3,4-tetrahydro isoquinoline hydrobromide, (470) primaquine diphosphate, (471) pentaquine phosphate, (472) dibucaine hydrochloride, (473) 9-aminoacridine hydrochloride hemihydrate, (474) 3, 6-diamino acridine hemisulfate, (475) 2-quinoline thiol hydrochloride, (476) sparteine sulfate pentahydrate, (477) papaverine hydrochloride, (478) emetine dihydrochloride hydrate, (479) 1,10-phenanthroline monohydrochloride monohydrate, (480) neocuproine hydrochloride trihydrate, (481) pyrimidine, (482) 2 chloropyrimidine, (483) 4-phenylpyrimidine, (484) 5-bromopyrimidine, (485) 2,4-dichloropyrimidine, (486) 4,6-dichloropyrimidine, (487) 2,4-dichloro-6-methylpyrimidine, (488) 6-chloro-2,4-dimethoxypyrimidine, (489) 2-amino-4,6-dimethoxypyrimidine, (490) 2,4,6-trichloropyrimidine, (491) 2,4,5,6-tetrachloropyrimidine, (492) 1,3,4,6,7,8-hexahydro-1-methyl-2H-pyrimido [1,2-a] pyrimidine, (493) 1,3,4,6,7,8-hexahydro-2H-pyrimido [1,2-a] pyrimidine, (494) hexetidine, (495) tert-butyl S-(4,6-dimethylpyrimidin-2-yl) thiocarbonate, (496) 4-methoxybenzyl-S(4,6-dimethylpyrimidin-2-yl) thiocarbonate, (497) 2-amino pyrimidine, (498) 2-amino-4-methyl pyrimidine, (499) 2-amino-5-nitropyrimidine, (500) 2-amino-5-bromopyrimidine, (501) 2-amino-4-chloro-6-methyl pyrimidine, (502) 2-amino-4,6-dimethyl pyrimidine, (503) 2-amino-4-hydroxy-6-methyl pyrimidine, (504) 2-amino-4,6-dichloropyrimidine, (505) 2-amino-5-bromo-6-methyl-4-pyrimidinol, (506) 4-aminopyrimidine, (507) 4,5-diamino pyrimidine, (508) 4-amino-2,6-dimethyl pyrimidine, (509) 2,4-diamino-6-hydroxypyrimidine, (510) 2,6-diamino-4-chloro pyrimidine, (511) 4,6-diamino-2-mercaptopyrimidine hemihydrate, (512) 2,4,6-triamino pyrimidine, (513) 5-nitroso-2,4,6-triamino pyrimidine, (514) 4,6-dihydroxy pyrimidine, (515) 4,6-dihydroxy-2-amino pyrimidine, (516) 4,6-dihydroxy-2-methyl pyrimidine, (517) 4,6-dihydroxy-5-nitropyrimidine, (518) 2,4-dihydroxy-5-methyl pyrimidine, (519) 2,4-dihydroxy-6-methyl pyrimidine, (520) 2,4-dihydroxy-5,6-dimethyl pyrimidine, (521) 2,6-dihydroxy pyrimidine-5-carboxylic acid hydrate, (522) 2,6-dihydroxy-4-amino pyrimidine, (523) 2,4,5-trihydroxy pyrimidine, (524) 2-thiouracil, (525) 6-amino-5-nitroso-2-thiouracil, (526) folic acid dihydrate, (527) folinic acid, calcium salt hydrate, (528) 2-hydroxypyrimidine hydrochloride, (529) 2-hydroxy-4-methyl pyrimidine hydrochloride, (530) 4,6-dimethyl-2-hydroxypyrimidine hydrochloride, (531) 2-mercapto-4-methyl pyrimidine hydrochloride, (532) 4,6-diamino pyrimidine hemisulfate monohydrate, (533) 4,5,6-triamino pyrimidine sulfate hydrate, (534) 4,5-diamino-6-hydroxy pyrimidine sulfate, (535) 2,4-diamino-6-mercapto pyrimidine hemisulfate, (536) 2,4-diamino-6-hydroxy pyrimidine hemisulfate hydrate, (537) 6-hydroxy-2,4,5-triamino pyrimidine sulfate, (538) 5,6-diamino-2,4-dihydroxy pyrimidine sulfate, (539) N4-(2-amino-4-pyrimidinyl) sulfanilamide monohydrochloride, (540) 2,4,5,6-tetraamino pyrimidine sulfate, (541) 2,4 (1H,3H)-pyrimidine dione, (542) 5-amino uracil, (543) 5-nitrouracil, (544) 5-iodouracil, (545) 5-(hydroxymethyl) uracil hydrate, (546) 5,6-dihydrouracil, (547) 6-amino-1-methyl uracil, (548) 5,6-diamino-1,3-dimethyl uracil hydrate, (549) uridine, (550) 5-methyl uridine, (551) 5-iodouridine, (552) thimidine, (553) 5-methyl-2-thiouracil, (554) 4-thiouridine, (555) 2-thiocytidine dihydrate, (556) orotic acid monohydrate, (557) hydroorotic acid, (558) 5-aminoorotic acid, (559) methylorotate, (560) barbituric acid, (561) 5-nitrobarbituric acid trihydraet, (562) violuric acid monohydrate, (563) alloxan monohydrate, (564) 4,5,6-triamino-2(1H)-pyrimidinethione sulfate, (565) cyclocytidine hydrochloride, (566) cytosine arabinoside hydrochloride, (567) pyridazine, (568) phthalazine, (569) 4,5-dihydro-6-methyl-3(2H)-pyridazinone monohydrate, (570) 3,6-dichloropyridazine, (571) 3,4,5-trichloropyridazine, (572) 3,6-dichloro-4-methylpyridazine, (573) 3-chloro-6-methoxypyridazine, (574) pyrazine, (575) acetylpyrazine, (576) aminopyrazine, (577) 2,6-dichloropyrazine, (578) 2,3,5-trimethylpyrazine, (579) tetramethylpyrazine, (580) 5-methyl-2-pyrazine carboxylic acid, (581) pyrazine amide, (582) 2,3-pyrazine dicarboxamide, (583) 4-pyridazine carboxylic acid, (584) 2,3-pyrazine dicarboxylic acid, (585) lumazine monohydrate, (586) xanthopterin monohydrate, (587) 2-quinoxazoline carboxylic acid, (588) 2-quinoxalinol, (589) 2,3-dihydroxy quinoxaline, (590) phenazine methosulfate, (591) 2-azetidinone, (592) 2-pyrrolidinone, (593) pyrrolidone hydrotribromide, (594) δ-valerolactam, (595) ε-caprolactam, (596) amino-ε-caprolactam, (597) N-methyl caprolactam, (598) 2-azacyclooctanone, (599) 2-azacyclononanone, (600) ω-thiocaprolactam, (601) N-vinylcaprolactam, (602) 2-azabicyclo[2.2.1]hept-5-en-3-one, (603) maleimide, (604) N-ethylmaleimide, (605) N-butylmaleimide, (606) N-cyclohexylmaleimide, (607) N-phenylmaleimide, (608) N-benzylmaleimide, (609) N-hydroxymaleimide, (610) succinimide, (611) N-methylsuccinimide, (612) 2-hydroxy-N-methylsuccinimide, (613) N-hydroxysuccinimide, (614) succinimidyl 2,2,2-trichloroethyl carbonate, (615) 2-dodecyl-N-(2,2,6,6-tetramethyl-4-ppiperidinyl) succinimide, (616) 2-dodecyl-N-(1,2,2,6,6-pentamethyl-4-piperdinyl) succinimide, (617) N-(1-acetyl-2,2,6,6-tetramethyl-4-piperidinyl)-2-dodecyl succinimide, (618) α-methyl-α-propylsuccinimide, (619) α-methyl-α-phenylsuccinimide, (620) N-vinylphthalimide, (621) N-ethylphthalimide, (622) N-(trimethylsilylmethyl)phthalimide, (623) N-(2-bromoethyl)phthalimide, (624) N-(3-bromopropyl)phthalimide, (625) N-(4-bromobutyl)phthalimide, (626) phthalimidoacetaldehyde diethyl acetal, (627) diethyl (phthalimidomethyl)phosphonate, (628) N-benzylphthalimide, (629) phthalimide, DBU (1,8-diazabicyclo [5.4.0]undec-7-ene) salt, (630) phthalimide, DBN (1,5-diazabicyclo [4.3.0]non-5-ene), and (631) mixtures thereof; or wherein the transparentizing agent is an oxa-aza-cyclic compound; or wherein the transparentizing agent is selected from the group consisting of: (A) materials of the general formulae: wherein R₁, R₂, R₃, R₄, R₅, R₆, R₇, R₈, R₉, R₁₀, R₁₁, R₁₂, R₁₃, R₁₄, and R₁₅ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, R₁₄, and R₁₅ can be joined together to form a ring; (B) materials of the general formula: wherein R₁, R₂, R₃, R₄, R₅, and R₆ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, and R₆ can be joined together to form a ring; (C) mixtures thereof; or wherein the transparentizing agent is selected from the group consisting of (1) 3-amino-5-methyl isoxazole, (2) 5-amino-3-methyl isoxazole, (3) 3,5-dimethyl-4-nitroisoxazole, (4) 1,2-benzisoxazole, (5) 2,1-benzisoxazole, (6) cycloserine, (7) 4-benzyl-2-methyl-2-oxazoline, (8) 2-methyl-5-phenyl-2-oxazoline-4-methanol, (9) benzoxazole, (10) 2-methylbenzoxazole, (11) 2-chlorobenzoxazole, (12) 2-chloro-3-ethylbenzeneoxazolium tetrafluoroborate, (13) 2-oxazolidone, (14) 3-methyl-2-oxazolidinone, (15) 5-chloromethyl-2-oxazolidinone, (16) 4-isopropyl-2-oxazolidinone, (17) 3-acetyl-2-oxazolidinone, (18) 5,5-dimethyl oxazolidine-2,4-dione, (19) 3-ethyl-2-thioxo-4-oxazolidinone, (20) 4-methyl-5-phenyl-2-oxazolidinone, (21) 4-benzyl-2-oxazolidinone, (22) 2-benzoisoxazolinone, (23) muscimol hydrate, (24) 5-methyl-3-phenyl isoxazole-4-carboxylic acid, (25) 2-methyl-5-phenyl-2-oxazoline-4-methanol, (26) sulfamethoxazole, (27) sulfisoxazole, (28) N'-(4,5-dimethyloxazol-2-yl) sulfanilamide, (29) chlorzoxazone, (30) 3,3'-dimethyl oxacarbocyanine iodide, (31) 2-ethyl-5-phenyl isoxazolium-3'-sulfonate, (32) 2-tert-butyl-5-methyl isoxazolium perchlorate, (33) 5-phenyl-2-(4-pyridyl) oxazole hydrochloride hydrate, (34) 5-phenyl-2-(4-pyridyl) oxazole methyl tosylate salt, (35) 4-aminomorpholine, (36) 4-morpholine carbonitrile, (37) 4-morpholine propionitrile, (38) 4-formyl morpholine, (39) 4-acetylmorpholine, (40) 4-(2-hydroxyethyl) morpholine, (41) 3-morpholino-1,2-propane diol, (42) 4-(3-amino propyl) morpholine, (43) 1-morpholino-1-cyclopentene, (44) 1-morpholino-1-cyclohexene, (45) 1-morpholino-1-cycloheptene, (46) 4-phenyl morpholine, (47) 4-morpholinoaniline, (48) 2,2,2-tribromoethyl phosphoromorpholino chloridate, (49) 1-(morpholino carbonyl methyl) piperazine, (50) 1,3-dimorpholine-2-nitropropane, (51) hemicholinium-3, (52) hemicholinium-15, (53) 2-methoxy-4-morpholinobenzene diazoniumchloride, zinc chloride, (54) fomocaine, (55) 4-morpholinobenzophenone, (56) 4,4'-ethylene-bis (2,6-morpholinedione), (57) N,N'-dicylcohexyl-4-morpholine carboxamidine, (58) 1-cyclohexyl-3-(2-morpholino ethyl)-2-thiourea, (59) 4-morpholinoacetophenone, (60) 4-(2-chloroethyl) morpholine hydrochloride, (61) 4-morpholine ethane sulfonic acid, (62) 4-morpholine propane sulfonic acid, (63) β-hydroxy morpholine propane sulfonic acid, (64) [N-(aminoiminomethyl)-4-morpholine carboximidamide] hydrochloride, (65) 4-morpholine carbodithioic acid compound with morpholine, (66) 2,5-dimethyl-4-(morpholinomethyl) phenol hydrochloride monohydrate, (67) 1-cyclohexyl-3-(2-morpholinoethyl) carbodiimide metho-p-toluene sulfonate, (68) hemicholinium-3[2,2'-(4,4'-biphenylene) bis(2-hydroxy-4,4-dimethyl morpholinium bromide), (69) hemicholinium-15[4,4-dimethyl-2-hydroxy-2-phenyl morpholinium bromide], (70) 1-aza-12-crown-4, (71) 1-aza-15-crown-5, (72) 1-aza-18-crown-6, (73) 1,4,10-trioxa-7,13-diazacyclopentadecane, (74) 1,4,10,1 3-tetraoxa-7,16-diazacyclooctadecane, (75) N,N'-dibenzyl-1,4,10,13-tetraoxa-7,16-diazacyclooctadecane, (76) 4,7,13,18-tetraoxa-1,10-diazabicyclo [8.5.5] eicosane, (77) 4,7,13,16,21-pentaoxa-1,10-diazabicyclo [8.5.5] tricosane, (78) 4,7,13,16,21,24-hexaoxa-1,10-diazabicyclo [8.8.8] hexacosane, (79) 5,6-benzo-4,17,13,16,21,24-hexaoxa-1,10-diazabicyclo[8.8.8] hexacosane, and (80) mixtures thereof; or wherein the transparentizing agent is an oxacyclic compound; or wherein the transparentizing agent is selected from the group consisting of: (A) materials of the general formula: wherein the curved portion of the structure represents a hydrocarbon chain or a substituted hydrocarbon chain, wherein two or more substituents can be joined together to form a ring; (B) materials of the general formulae: wherein R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, and R₂₈ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, and R₂₈ can be joined together to form a ring; (C) materials of the general formula: wherein the curved portion of the structure represents a hydrocarbon chain or a substituted hydrocarbon chain, wherein two or more substituents can be joined together to form a ring; (D) materials of the general formulae: wherein R₁, R₂, R₃, R₄, R₅, R₆, R₇, and R₈ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, and R₈ can be joined together to form a ring; (E) materials of the general formulae: wherein the curved portions of the structures represent a hydrocarbon chain or a substituted hydrocarbon chain, wherein two or more substituents can be joined together to form a ring; (F) materials of the general formula: wherein R₁, R₂, R₃, R₄, R₅, and R₆ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, and R₆ can be joined together to form a ring; and (G) mixtures thereof; or wherein the transparentizing agent is selected from the group consisting of (1) γ-butyrolactone, (2) γ-valerolactone, (3) γ-caprolactone, (4) γ-octanoic lactone, (5) γ-nonanoic lactone, (6) γ-decanolactone, (7) undecanoic γ-lactone, (8) γ-phenyl-γ-butyrolactone, (9) α-carbethoxy-γ-phenyl-butyrolactone, (10) 2-coumaranone, (11) β,β-dimethyl-γ-(hydroxymethyl)-γ-butyrolactone, (12) γ-ethoxy carbonyl-γ-butyrolactone, (13) 5-(hydroxymethyl)-2(5H)-furanone, (14) dihydro-4,4-dimethyl-2,3-furandione, (15) 2,5-dimethyl-4-hydroxy-3(2H)-furanone, (16) mevalonic (β-hydroxy β-methyl-δ-valero) lactone, (17) δ-decanolactone, (18) undecanoic δ-lactone, (19) δ-dodecanolactone, (20) undecanoic ω-lactone, (21) oxacyclotridecan-2-one, (22) ω-pentadecalactone, (23) hydrindantin (2,2'-dihydroxy-2,2'-biindan-1,1'3,3'-tetrone, (24) hydrindantin dihydrate, (25) 2-oxepanone, (26) 4H-pyran-2-one, (27) methylcoumalate, (28) methyl 2-oxo-2H-pyran-3-carboxylate, (29) 4,6-dimethyl-α-pyrone, (30) 4-methoxy-6-methyl-2H-pyran-2-one, (31) 3,6-dihydro-4,6,6-trimethyl-2H-pyran-2-one, (32) 3,4-dihydro-6-methyl-2H-pyran-2-one, (33) 3-acetyl coumarin, (34) 6-methyl coumarin, (35) 7-ethoxy coumarin, (36) ethyl-3-coumarin carboxylate, (37) 7-diethylamino-4-methyl coumarin, (38) dihydro coumarin, (39) 3-bromo-2-coumaranone, (40) patulin, (41) 4H-pyran-4-one, (42) 2-ethyl-3-hydroxy-4H-pyran-4-one, 43v) butopyronoxyl(butyl 3,4-dihydro-2,2-dimethyl-4-oxo-2H-pyran-6-carboxylate, (44) dehydroacetic acid, (45) 4-chromone, (46) 4-chromanone, (47) 4-chromanol, (48) 6,7-dimethoxy-2,2-dimethyl-4-chromanone, (49) 3-isochromanone, (50) 6,7-dimethoxy-3-isochromanone, (51) 6-ethyl-4-oxo-4H-1-benzopyran-3-carbonitrile, (52) 6-ethyl-4-oxo-4H-1-benzopyran-3-carboxaldehyde, (53) 6-isopropyl-4-oxo-4H-1-benzopyran-3-carbonitrile, (54) 6-isopropyl-4-oxo-4H-1-benzopyran-3-carboxaldehyde, (55) maleic anhydride, (56) bromomaleic anhydride, (57) citraconic anhydride, (58) 2,3-dimethylmaleic anhydride, (59) dichloromaleic anhydride, (60) cis-aconitic anhydride, (61) itaconic anhydride, (62) methylsuccinic anhydride, (63) acetylmercaptosuccinic anhydride, (64) 2,2-dimethylsuccinic anhydride, (65) phenylsuccinic anhydride, (66) 2-octen-1-ylsuccinic anhydride, (67) 2-dodecen-1-ylsuccinic anhydride, (68) 2-octadecen-1-ylsuccinic anhydride, (69) 3-oxabicyclo [3.1.0] hexane-2,4-dione, (70) diglycolic anhydride, (71) glutaric anhydride, (72) 3-methylglutaric anhydride, (73) 2,2-dimethylglutaric anhydride, (74) 3,3-tetramethyleneglutaric anhydride, (75) 1-cyclopentene-1,2-dicarboxylic anhydride, (76) 3,4,5,6-tetrahydrophthalic anhydride, (77) cis-1,2-cyclohexanedicarboxylic anhydride, (78) hexahydro-4-methylphthalic anhydride, (79) methyl-5-norbornene-2,3-dicarboxylic anhydride, (80) 2,3-pyridinecarboxylic anhydride, (81) 3,4-pyridinecarboxylic anhydride, (82) furfurylmercaptan, (83) S-furfurylthioacetate, (84) furfurylsulfide, (85) furfurylmethyldisulfide, (86) furfuryldisulfide, (87) glycolaldehyde dimer, (88) 6,7-dihydrocyclopenta-1,3-dioxin-5(4H)-one, (89) (2R,6R)-tert-butyl-6-methyl-1,3-dioxan-4-one, (90) 2,2-dimethyl-1,3-dioxane-4,6-dione, (91) 3,6-dimethyl-1,4-dioxane-2,5-dione, (92) 2,2,6-trimethyl-4H-1,3-dioxin-4-one, (93) 2,2,5-trimethyl-1,3-dioxane-4,6-dione, (94) 5-bromo-2,2,5-trimethyl-1,3-dioxane-4,6-dione, (95) 1,3-dioxane-5,5-dimethanol, (96) 1,3,5-trioxane, (97) 1,6-dioxaspiro [4.4]nonane-2,7-dione, (98) 1,4-dioxaspiro [4.5]decan-2-one, (99) 1,7-dioxaspiro [5.5]undecane, (100) 2,4,8,10-tetraoxaspiro[5.5]undecane, (101) 3,9-divinyl-2,4,8-tetraoxaspiro[5.5]undecane, (102) 2,2-pentamethylene-1,3-dioxalane, (103) 2-phenyl-1,3-dioxalane, (104) 1,4-cyclohexanedione monoethylene ketal, (105) 1,4-cyclohexanedione bis(ethylene ketal), (106) 1,4-cyclohexanedione mono-2,2-dimethyl trimethylene ketal, (107) piperonal, (108) piperonyl acetate, (109) piperonyl alcohol, (110) piperonylnitrile, (111) piperonyl amine, (112) 6-nitropiperonal, (113) 6-nitropiperonyl alcohol, (114) 3',4'-(methylenedioxy)acetophenone, (115) 3,4-(methylenedioxy)aniline, (116) 2,3-(methylenedioxy)benzaldehyde, (117) 3,4-(methylenedioxy)phenylacetonitrile, (118) 3,4-(methylenedioxy)toluene, and (119) mixtures thereof; or wherein the transparentizing agent is a crown ether; or wherein the transparentizing agent is selected from the group consisting of (1) 1,4,7,10-tetraoxacyclododecane (12-crown-4), (2) 2-(hydroxyethyl)-12-crown-4, (3) 2-(aminoethyl)-12-crown-4, (4) benzo-12-crown-4, (5) 1,4,7,10,13-pentaoxacyclododecane (15-crown-5), (6) 2-(hydroxyethyl)-15-crown-5, (7) 2-(aminoethyl)-15-crown-5, (8) benzo-15-crown-5, (9) 4'-aminobenzo-15-crown-5, (10) 4'-formylbenzo-15-crown-5, (11) 4'-nitrobenzo-15-crown-5, (12) bis [(benzo-15-crown-5)-15-ylmethyl] pimelate, (13) 1,4,7,10,13,16-hexaoxacyclooctadecane (18-crown-6), (14) 2-(aminoethyl)-18 crown-6, (15) benzo-18 crown-6, (16) 4'-bromobenzo-18-crown-6, (17) dibenzo-18-crown-6, (18) di-tert-butyldibenzo-18-crown-6, (19) cis-dicyclohexane-18 crown-6, (20) dibenzo-24-crown-8, (21) dicyclohexano-24-crown-8, (22) dibenzo-30-crown-10, and (23) mixtures thereof; or wherein the transparentizing agent is a cyclic hydrocarbon; or wherein the transparentizing agent is selected from the group consisting of: (A) materials of the general formulae: wherein R₁, R₂, R₃, R₄, R₅, R₆, R₇, R₈, R₉, R₁₀, R₁₁, and R₁₂ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, and R₁₂ can be joined together to form a ring; (B) materials of the general formula: wherein R₁, R₂, R₃, R₄, R₅, and R₆ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, and R₆ can be joined together to form a ring; (C) materials of the general formula: wherein R₁, R₂, R₃, R₄, R₅, R₆, R₇, R₈, R₉, and R₁₀ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, and R₁₀ can be joined together to form a ring; (D) materials of the general formulae: wherein R₁, R₂, R₃, R₄, R₅, R₆, R₇, R₈, R₉, R₁₀, R₁₁, and R₁₂ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, R₁₀, R₁₁, and R₁₂ can be joined together to form a ring; (E) materials of the general formula: wherein R₁, R₂, R₃, R₄, R₅, R₆, R₇, R₈, R₉, and R₁₀ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, and R₁₀ can be joined together to form a ring; (F) materials of the general formulae: wherein R₁, R₂, R₃, R₄, R₅, R₆, R₇, R₈, R₉, and R₁₀ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R₂, R₃, R₄, R₅, R₆, R₇, R₈, R₉, and R₁₀ can be joined together to form a ring; (G) materials of the general formula: wherein the curved portion of the structure represents a hydrocarbon chain or a substituted hydrocarbon chain, wherein two or more substituents can be joined together to form a ring; and (H) mixtures thereof; or wherein the transparentizing agent is selected from the group consisting of (1) norbornane, (2) 2-norbornane carbonitrile, (3) 2-norbornane methanol, (4) 3-methyl-2-norbornane methanol, (5) camphene, (6) fenchyl alcohol, (7) thiocamphor, (8) norbornene, (9) 5-norbornene-2-carbonitrile, (10) 5-norbornene-2-carboxaldehyde, (11) 5-norbornene-2-methanol, (12) 5-norbornene-2,2-dimethanol, (13) 5-norbornene-2-benzoyl, (14) 2-norbornanone, (15) 3-chloro-2-norbornanone, (16) fenchone, (17) 3-(trifluoroacetyl)camphor, (18) 3-heptafluorobutyryl camphor, (19) 3-bromocamphor, (20) 9,10-dibromocamphor, (21) 3,9,10-tribromocamphor, (22) dicyclopentadiene, (23) methylcyclopentadiene dimer, (24) tricyclo[5.2.1]decane, (25) 4,8-bis(hydroxymethyl)tricyclo[5.2.1.0^{2.6}]decane, (26) 8-ketotricyclo[5.2.1.0^{2.6}]decane, (27) 3,4-dimethoxy-3-cyclobutene-1,2-dione, (28) 3,4-diethoxy-3-cyclobutene-1,2-dione, (29) 3,4-diisopropoxy-3-cyclobutene-1,2-dione, (30) 3,4-dibutoxy-3-cyclobutene-1,2-dione, (31) 3-methyl-2-(nitromethyl)-5-oxocyclopentaneacetic acid, (32) 3-ethyl-2-hydroxy-2-cyclopenten-1-one, (33) methyl-4-methoxy-2-oxo-3-cyclopentene-1-carboxylate, (34) 3,3a,6,6a-tetrahydro-2H-cyclopenta[b]furan-2-one, (35) 3a,4,5,6a-hexahydro-5-hydroxy-4(hydroxymethyl)-2H-cyclopenta[b]furan-2-one, (36) 3-methyl-1,2-cyclopentanedione, (37) 4-hydroxy-5-methyl-4-cyclopentene-1,3-dione monohydrate, (38) 2,4,4-trimethylcyclohexen-1-one, (39) ethyl-6-methyl-2-oxo-3-cyclohexene-1-carboxylate, (40) ethyl 4-hydroxy-6-methyl-2-oxo-3-cyclohexene-1-carboxylate, (41) 5-(1-acetoxy-1-methylethyl)-2-methyl-2-cyclohexen-1-one, (42) thymoquinone, (43) 2,6,6-trimethyl-2-cyclohexene-1,4-dione, (44) indan, (45) 1-indanol, (46) 2-indanol, (47) 1-indanone, (48) 2-indanone, (49) 2-acetyl-1-tetralone, (50) 4-methyl-1-tetralone, 513) 5,7-dimethyl-1-tetralone, (52) 6,7-dimethoxy-1-tetralone, (53) 1-methyl-2-tetralone, (54) 6,7-dimethoxy-2-tetralone, (55) cyclohexanone, (56) cycloheptanone, (57) cyclooctanone, (58) cyclononanone, (59) cyclodecanone, (60) cycloundecanone, (61) cyclododecanone, (62) cyclotridecanone, (63) cyclopentadecanone, (64) 2-acetylcyclohexanone, (65) 2-allylcyclohexanone, (66) 2-phenylcyclohexanone, (67) cyclohexanedione, (68) 2-acetyl-1,3-cyclohexanedione, (69) 4,4-dimethyl-1,3-cyclohexanedione, (70) 2-acetyl-1,3-cyclopentanedione, (71) 3,3,5,5-tetramethyl-1,2-cyclopentanedione, (72) bicyclo[3.2.1]octan-2-one, (73) endo-dimethyl 7-oxabicyclo[2.2.1]heptane-2,3-dicarboxylate, (74) cineole, (75) bicyclo[2.2.2]oct-5-ene-2,3-dimethanol, (76) tropone, (77) tropolone, (78) cyclooctene oxide, (79) 1,2,5,6-diepoxycyclooctane, (80) 9-methyl-Δ⁵⁽¹⁰⁾-octalin-1,6-dione, (81) cis-bicyclo[3.3.0]octane-3.7-dione, (82) azulene, (83) 1-benzosuberone, (84) 1,5,9-cyclododecatriene, (85) cyclododecane epoxide, (86) 2,3-cyclododeceno pyridine, (87) 1,2,5,6,9,10-hexabromo cyclododecane, (88) 8-cyclohexadecen-1-one, (89) bicyclo[10.3.0]pentadec-12(1)-en-13-one, (90) 1,4,4a,8a-tetrahydro-endo-1,4-methanonaphthalene-5,8-dione, and (19) mixtures thereof; or wherein the transparentizing agent is a thiourea; or wherein the transparentizing agent is a sulfone; or wherein the transparentizing agent is a thiocyclic compound; or wherein the transparentizing agent is selected from the group consisting of sulfites, sulfite derivatives, sulfides, sulfide derivatives, quaternary sulfur compounds, quaternary sulfur derivatives, and mixtures thereof; or wherein the transparentizing agent is a thia-aza-cyclic compound; or wherein the transparentizing agent is selected from the group consisting of (1) 1-allyl-2-thioure, (2) 1-methallyl-3-methyl-2-thiourea, (3) 4-allyl-3-thiosemicarbazide, (4) 1,3-diethyl-2-thiourea, (5) 1,3-dibutyl-2-thiourea, (6) 1-benzyl-3-methyl-2-thiourea, (7) 1,1,3,3-tetramethyl-2-thiourea, (8) 2-imino-4-thiobiuret, (9) 1-allyl-3-(2-hydroxyethyl)-2-thiourea, (10) S-(2-aminoethyl)isothiouronium bromide hydrobromide, (11) S,S-diphenylsulfillimine monohydrate, (12) methylsulfon), (13) ethylsulfone, (14) butylsulfone, (15) butadiene sulfone, (16) tetramethylene sulfone, (17) 1,4-butane sulfone, (18) 1,4-butanediolcyclic sulfate, (19) benzylsulfone, (20) phenylsulfone, (21) phenylvinylsulfone, (22) phenylstyrenesulfone, (23) phenyl-2-(trimethylsilyl)methyl sulfone, (24) phenyl 2-(trimethylsilyl)ethyl sulfone, (25) phenyl 2-(trimethylsilyl)ethynyl sulfone, (26) 4-(fluorophenyl)sulfone, (27) 4-(fluorophenyl)methyl sulfone, (28) chloromethylphenyl sulfone, (29) chloromethyl-p-tolyl sulfone, (30) 2-chloroethylphenyl sulfone, (31) methylthiomethylphenyl sulfone, (32) methylthiomethyl-p-tolyl sulfone, (33) 2-(phenylsulfonyl) tetrahydropyran, (34) 1-(phenylsulfonyl)indole, (35) 1-(p-toluenesulfonyl)imidazole, (36) 1-(p-tosyl)-3,4,4-trimethyl imidazolidine, (37) 4-(p-tosylsulfonyl)hexahydro -1,4-thiazepine, (38) thionaphthene, (39) 4-keto-4,5,6,7-tetrahydrothianaphthene, (40) 2,2'-bithiophene, (41) 2,2':5',2"-terthiophene, (42) N-acetylhomocysteine thiolactone, (43) tetrahydrothiopyran-4-one, (44) thiochroman-4-one, (45) thiochroman-4-ol, (46) thioctic acid, (47) ethyl 1,3-dithiolane-2-carboxylate, (48) 3H-1,2-benzodithiol-3-one, (49) 1,3-dithiane, (50) 2-phenyl-1,3-dithiane, (51) ethyl-1,3-dithiane-2-carboxylate, (52) 5,6-dihydro-5-methyl-4H-1,3,5-dithiazine, (53) 1,4-dithiane, (54) 2,5-dihydroxy-2,5-dimethyl-1,4-dithiane, (55) 1,5-dithiacyclooactan-3-ol, (56) 1,4-dithiaspiro [45] decan-8-ol, (57) 1,3,5-trithiane, (58) 1,4,7-trithiacyclononane, (59) 1,4,7-trithiacyclodecane, (60) 1,4,7,10-tetrathiacyclododecane, (61) 3,6,9,14-tetrathiabicyclo [9.2.1] tetradeca-11,13-diene, (62) 1,4,8,1-tetrathiacyclotetradecane, (63) 1,5,9,13-tetrathiocyclohexadecane, (64) 1,5,9,13-tetrathiacyclohexadecane-3,11-diol, (65) 1,4,7,10,13-pentathiacyclopentadecane, (66) 1,4,7,10,13,16-hexathiacyclooctadecane, (67) 1,5,9,13,17,21-hexathiacyclotetracosane-3,1 1,19-triol, (68) 1,4,7,10,13,16,19,22-octathiacyclotetracosane, (69) 1,4,8,11,15,18,22,25-octathiacyclooctacosane, (70) 1,4,7,10,13,16,19,22,25-nonathiacycloheptacosane, (71) dimethylsulfite, (72) diethylsulfite, (73) sodium sulfite, (74) allyldisulfide, (75) aminophenyldisulfide, (76) benzyldisulfide, (77) benzylphenylsulfide, (78) trimethylsulfonium methylsulfate, (79) (2-chloroethyl)dimethylsulfonium iodide, (80) 3-(chloropropyl)diphenylsulfonium tetrafluoroborate, (81) trimethyl sulfonium iodide, (82) trimethyl sulfoxonium iodide, (83) trimethyl sulfoxonium chloride, (84) triphenyl methane sulfenyl chloride, (85) dimethyl (2-methoxy-5-nitrobenzyl) sulfonium bromide, (86) thionin perchlorate, (87) p-xylylene bis(tetrahydrothiopheneum chloride), (88) tris (dimethyl amino) sulfonium difluorotrimethyl silicate, (89) tris (dimethyl amino) sulfonium trifluoromethoxide, (90) (3-amino-3-carboxypropyl) dimethyl sulfonium chloride, and (91) mixtures thereof; or wherein the transparentizing agent is of one of the general formulae: wherein R₁, R₂, R₃, R₄, R₅, R₆, and R₇ each, independently of the others, are selected from the group consisting of hydrogen atoms, alkyl groups, substituted alkyl groups, aryl groups, substituted aryl groups, arylalkyl groups, substituted arylalkyl groups, hydroxy groups, amine groups, imine groups, ammonium groups, pyridine groups, pyridinium groups, ether groups, aldehyde groups, ketone groups, ester groups, amide groups, carboxylic acid groups, carbonyl groups, thiocarbonyl groups, sulfate groups, sulfonate groups, sulfide groups, sulfoxide groups, phosphine groups, phosphonium groups, phosphate groups, cyano groups, nitrile groups, mercapto groups, nitroso groups, halogen atoms, nitro groups, sulfone groups, acyl groups, acid anhydride groups, and azide groups, wherein two or more of R₁, R2, R3, R4, R₅, R6, and R7 can be joined together to form a ring; or wherein the transparentizing agent is selected from the group consisting of (1) 2-amino-2-thiazoline, (2) 2-amino thiazole, (3) 2-amino-4-methylthiazole, (4) 2-amino-4-methylthiazole, (5) 2-amino-4-thiazoleacetic acid, (6) 2-acetamido-4-methylthiazole, (7) 2-acetylthiazole, (8) 5-acetyl-2,4-dimethylthiazole, (9) 4-methyl-5-vinylthiazole, (10) 2-amino-4-phenyl-5-tetradecylthiazole, (11) 2,4-thiazolidine dione, (12) 3-aminorhodanine, (13) 3-methylrhodanine, (14) 3-ethylrhodanine, (15) 3-allylrhodanine, (16) 3-hydroxy-4-methyl-2(3H)-thiazolethione, (17) benzothiazole, (18) 2-methylbenzothiazole, (19) 2-(methylthio)benzothiazole, (20) 2-amino-4-methylbenzothiazole, (21) 3-methylbenzothiazole-2-thione, (22) 2,1,3-benzothiadiazole, (23) 4-amino-2,1,3-benzothiadiazole, (24) 3,4-dimethyl-5-(2-hydroxyethyl)thiazolium iodide, (25) 3-ethyl-5-(2-hydroxyethyl)4-methylthiazolium bromide, (26) 2-amino-5-nitrothiazole, (27) 2-amino-α-(methoxyimino)-4-thiazole acetic acid, (28) ethyl 2-amino-a-(hydroxyimino)-4-thiazole acetate, (29) ethyl 2-amino-a-(methoxyimino)-4-thiazole acetate, (30) ethyl 2-amino-4-thiazole acetate, (31) ethyl 2-amino-4-thiazole glyoxylate, (32) 1-phenyl-3-(2-thiazolyl)-2-thiourea, (33) 2-amino-4-methoxy benzothiazole, (34) 2-amino-5,6-dimethylbenzothiazole, (35) N'-(2-thiazolyl) sulfanilamide, 6-ethoxy-2-benzothiazole sulfonamide, (37) ethyl-2-(formylamino)-4-thiazoleacetate, (38) ethyl-2-(formylamino)-4-thiazoleglyoxylate, (39) 2-(formylamino)-α-(methoxyimino)-4-thiazole acetic acid, (40) 2-acetamido-4-methyl-5-thiazole sulfonyl chloride, (41) 2-thioxo-4-thiazolidine carboxylic acid, (42) thiazolidine-4-carboxylic acid, (43) pseudothiohydantoin, (44) 2-amino-1,3,4-thiadiazole, (45) 2-amino-5-trifluoromethyl-1,3,4-thiadiazole, (46) 2-amno-5-methyl-1,3,4-thiadiazole, (47) 2-amino-5-ethyl-1,3,4-thiadiazole, (48) 2-amino-5-(ethylthio)-1,3,4-thiadiazole, (49) 5-amino-1,3,4-thiadiazole-2-thiol, (50) 2-acetamido-5-benzyl thio-1,3,4-thiadiazole, (51) 5-acetamido-1,3,4-thiadiazole-2-sulfonamide, (52) 5-anilino-1,2,3,4-thiatriazole, (53) 2-amino-4,5-dimethyl thiazole hydrochloride, (54) 2-amino 4-imino-2-thiazoline hydrochloride, (55) 2-amino-2-thiazoline hydrochloride, (56) 2-amino-5-bromothiazole monohydrobromide, (57) 5-amino-3-methyl isothiazole hydrochloride, (58) 3-methyl-2-benzothiazolinone hydrazone hydrochloride hydrate, (59) 5-amino-2-methylbenzothiazole dihydrochloride, (60) 2,4-diamino-5-phenyl thiazole monohydrobromide, (61) 2-amino-4-phenyl thiazole hydrobromide monohydrate, (62) 2-(tritylamino)-α-(methoxyimino)-4-thiazole acetic acid hydrochloride, (63) (2,3,5,6-tetrahydro-6-phenylimidazo [2,1-b] thiazole hydrochloride, (64) 3-ethyl-2-methyl-2-thiazolium iodide, (65) 3-benzyl-5-(2-hydroxyethyl)-4-methyl thiazolium chloride, (66) thiamine hydrochloride, (67) 3-(carboxymethyl) benzothiazolium bromide, (68) 2-azido-3-ethyl benzothiazolium tetrafluoroborate, (69) 3-ethyl-2-methyl benzothiazolium iodide, (70) 2-methyl-3-propyl benzothiazolium iodide, (71) 3-ethyl-2-(2-hydroxy-1-propenyl) benzothiazolium chloride, (72) 3,6-dimethyl-2-(4-dimethyl aminophenyl) benzothiazolium bromide, (73) trifluoroperazine dihydrochloride, (74) thioridazine hydrochloride, (75) promethazine hydrochloride, (76) ethopropazine hydrochloride, (77) chlorpromazine hydrochloride, and (78) mixtures thereof; or wherein the transparentizing agent is selected from the group consisting of phosphines, phosphites, cyclic phosphorus compounds, phosphine oxides, quaternary phosphonium salts, and mixtures thereof; or wherein the transparentizing agent is selected from the group consisting of (1) triphenylphosphine, (2) tri-m-tolyl phosphine, (3) tris(3-methoxyphenyl)phosphine, (4) tris(4-chlorophenyl)phosphine, (5) tris(pentafluorophenyl)phosphine, (6) tricyclohexylphosphine, (7) tribenzylphosphine, (8) tri-2-furylphosphine, (9) bis (pyrrolidino)methoxy phosphone, (10) tetraphenylbiphosphine, (11) 1,3-bis(diphenylphosphino)propane, (12) 1,5-bis(diphenylphosphino)pentane, (13) 1,6-bis(diphenylphosphino)hexane, (14) isopropyl diphenyl phosphine, (15) diphenyl (p-tolyl) phosphine, (16) (4-bromophenyl) diphenyl phosphine, (17) diphenyl-2-pyridylphosphine, (18) dicyclohexylphenyl phosphine, (19) trimethyl phosphite, (20) triethyl phosphite, (21) tris(2-chloroethyl) phosphite, (22) tributyl phosphite, (23) triphenyl phosphite, (24) trimethyl phosphite copper iodide, (25) triethyl phosphite copper iodide, (26) dipropyl phosphite, (27) bis(2-ethylhexyl) phosphite, (28) bis(4-nitrobenzyl) phosphite, (29) 2,2'-ethylidene bis(4,6-di-tert-butylphenyl) fluorophosphite, (30) pentaerythritol diphenyl diphosphite, (31) 2-furyltetramethyl phosphorodiamidate, (32) diethyl(pyrrolidinomethyl)phosphonate, (33) cyclophosphamide monohydrate, (34) 2-chloro-1,3,2-dioxaphospholane-2-oxide, (35) N,N-diethyl-1,5-dihydro-2,4,3-benzodioxaphosphepin-3-amine, (36) 1,2-phenylene phosphochloridite, (37) 1,2-phenylene phosphochloridate, (38) 2-chloro-4H-1,3,2-benzodioxaphosphorin-4-one, (39) 2,4-bis(methylthio)-1,3-dithia-2,4-diphosphetane-2,4-disulfide, (40) triphenyl phosphine oxide, (41) tris(hydroxymethyl) phosphine oxide, (42) trimethoxy phosphine oxide, (43) triethoxy phosphine oxide, (44) triphenoxy phosphine oxide), (45) tris (2-butoxy ethoxy) phosphine oxide, (46) diphenyl phosphine oxide, (47) diphenyl (2,4,6-trimethylbenzoyl) phosphine oxide, (48) phenyl phosphinic acid, (49) diphenyl phosphate, (50) vinyl phosphonic acid, (51) propyl phosphonic acid, (52) pyrophosphoric acid, (53) triphenylphosphate, (54) tetrabutylphosphonium chloride, (55) tetrabutylphosphonium bromide, (56) hexadecyltributylphosphonium bromide, (57) stearyltributylphosphonium bromide, (58) azidotris(diethylamino)phosphonium bromide, (59) phosphonitrilic chloride trimer, (60) tetramethyl phosphonium bromide, (61) tetramethyl phosphonium chloride, (62) tetraethyl phosphonium bromide, (63) tetraethyl phosphonium chloride, (64) tetraethyl phosphonium iodide, (65) tetraphenyl phosphonium bromide, (66) tetraphenyl phosphonium chloride, (67) tetraphenyl phosphonium Iodide, (68) methyl triphenyl phosphonium bromide, (69) methyl triphenyl phosphonium iodide, (70) ethyl triphenyl phosphonium bromide, (71) n-propyl triphenyl phosphonium bromide, (72) isopropyl triphenyl phosphonium iodide, (73) cyclopropyl triphenyl phosphonium bromide, (74) n-butyl triphenyl phosphonium bromide, (75) isobutyl triphenyl phosphonium bromide, (76) hexyl triphenyl phosphonium bromide, (77) benzyl triphenyl phosphonium chloride, (78) bromomethyl triphenyl phosphonium bromide, (79) chloromethyl triphenyl phosphonium chloride, (80) 3-bromopropyl triphenyl phosphonium bromide, (81) 3-bromobutyl triphenyl phosphonium bromide, (82) 4-bromobutyl triphenyl phosphonium bromide, (83) 2-dimethyl aminoethyl triphenyl phosphonium bromide, (84) [(3-dimethyl amino) propyl] triphenyl phosphonium bromide, (85) 2-hydroxyethyl triphenyl phosphonium bromide, (86) (2-hydroxyethyl) triphenyl phosphonium chloride, (87) [3-hydroxy-2-methyl propyl] triphenyl phosphonium bromide, (88) [3-hydroxy-2-methyl propyl] triphenyl phosphonium bromide, (89) (2-hydroxybenzyl triphenyl phosphonium bromide, (90) (formyl methyl) triphenyl phosphonium chloride, (91) (methoxymethyl) triphenyl phosphonium chloride, (92) acetonyl triphenyl phosphonium chloride, (93) carbomethoxymethyl triphenyl phosphonium bromide, (94) (ethoxy carbonyl methyl) triphenyl phosphonium chloride, (95) carbethoxymethyl triphenyl phosphonium bromide, (96) (tert-butoxy carbonyl methyl) triphenyl phosphonium bromide, (97) phenacyl triphenyl phosphonium bromide, (98) (4-ethoxybenzyl) triphenyl phosphonium bromide, (99) 4-butoxybenzyl triphenyl phosphonium bromide, (100) 2-(1,3-dioxan-2-yl) ethyl] triphenyl phosphonium bromide, (101) (1,3-dioxolan-2-ylmethyl) triphenyl phosphonium bromide, (102) vinyl triphenyl phosphonium bromide, (103) allyl triphenyl phosphonium bromide, (104) allyl triphenyl phosphonium chloride, (105) propargyl triphenyl phosphonium bromide, (106) (3-trimethyl silyl-2-propynyl) triphenyl phosphonium bromide, (107) p-xylylene bis (triphenyl phosphonium bromide), and (108) mixtures thereof; or wherein the transparentizing agent is a nitrile; or wherein the transparentizing agent is selected from the group consisting of (1) cyanoacetohydrazide, (2) 4,4-dimethyl-3-oxopentanenitrile, (3) 1-cyano-N-methylthioformamide, (4) cyanomethyl N,N-dimethyl dithiocarbamate, (5) 4-hydroxy-3-methoxy-phenyl acetonitrile, (6) tosyl cyanide, (7) tosylmethyl isocyanide, (8) 5-fluoro-2-methyl benzonitrile, (9) 2-fluoro-5-methyl benzonitrile, (10) 4-(methylthio) benzonitrile, (11) 4-(dimethylamino) benzonitrile, (12) 3,4-dimethoxy benzonitrile, (13) 4-hydroxy-3-methoxy benzonitrile, (14) 4-(trans-4-pentyl cyclohexyl)benzonitrile, (15) 4'-pentyl-4'-biphenyl carbonitrile, (16) 4'-(pentyloxy)-4-biphenylcarbonitrile, (17) 4'-hexyl-4-biphenyl carbonitrile, (18) 4'-(hexyloxy)-4-biphenyl carbonitrile, (19) 4'-heptyl-4-biphenyl carbonitrile, (20) 4'-heptyloxy-4-biphenyl carbonitrile, (21) 4'-octyl-4-biphenyl carbonitrile, (22) 4'-(octyloxy)-4-biphenyl carbonitrile, (23) succinonitrile, (24) fumaronitrile, (25) 1,4-dicyano-2-butene, (26) (dimethyl aminomethylene)malononitrile, (27) (1-ethoxyethylidene)malononitrile, (28) α-chlorobenzylidenemalononitrile, (29) benzylidenemalononitrile, (30) 2-benzoyloxy-2-phenyl malononitrile, (31) O-(p-tosyl)isonitrosomalononitrile, (32) tetrafluorophthalonitrile, (33) iminodiacetonitrile, (34) phenylene diacetonitrile, (35) 3,3'-(4-formyl phenylimino) dipropionitrile, (36) tris (2-cyanoethyl) nitromethane, (37) 1,1,3,3-propanetetracarbonitrile, (38) tetracyanoethylene oxide, and (39) mixtures thereof; or wherein the transparentizing agent is selected from the group consisting of isothiocyanates, isocyanates, and mixtures thereof; or wherein the transparentizing agent is selected from the group consisting of (1) 4-azidophenyl isothiocyanate, (2) 1-naphthyl isothiocyanate, (3) 4-dimethyl amino-1-naphthyl isothiocyanate, (4) 1-isothiocyanato-4-(trans-4-propyl cyclohexyl) benzene, (5) 1-(trans-4-hexyl cyclohexyl)-4-isothiocyanato benzene, (6) 1-(4-trans-hexyl cyclohexyl)-4-[2-(4-isothio cyanatophenyl)] benzene, (7) 1-isothiocyanato-4-(trans-4-octylcyclohexyl) benzene, (8) 4-isothiocyanatophenyl-4-pentabicyclo [2.2.2] octane-1-carboxylate, (9) benzylthiocyanate, (10) guanidinethiocyanate, (11) methylene dithiocyanate, (12) 4,4'-methylene bis (phenyl isocyanate), (13) 4,4'-methylene bis (2,6-diethyl isocyanate), and (14) mixtures thereof; or wherein the transparentizing agent is selected from the group consisting of oxime compound, hydroxamic acid compounds, and mixtures thereof; or wherein the transparentizing agent is selected from the group consisting of (1) formamidoxime (2) acetaldoxime, (3) pyruvic aldehyde-1-oxime, (4) acetone oxime, (5) ethylchlorooximido acetate, (6) 2,3-butane dione monoxime, (7) 5-hydroxy pentenal oxime, (8) cyclopentanone oxime, (9) cyclohexanone oxime, (10) cyclooctanone oxime, (11) benzaldehyde oxime, (12) 2-nitrobenzaldehyde oxime, (13) salicyl aldoxime, (14) 2-isonitroso acetphenone, (15) 1-phenyl-1,2-propanedione 2-oxime, (16) 2-pyridine aldoxime, (17) nifuroxime, and (18) mixtures thereof; or wherein the transparentizing agent is a hydroxamic acid derivative; or wherein the transparentizing agent is selected from the group consisting of (1) acetohydroxamic acid, (2) suberohydroxamic acid, (3) mandelohydroxamic acid, (4) benzohydroxamic acid, (5) N-phenylbenzohydroxamic acid, and (6) mixtures thereof; or wherein the transparentizing agent is selected from the group consisting of alkyl ammonium salts, aryl ammonium salts, arylalkyl ammonium salts, and mixtures thereof; or wherein the transparentizing agent is selected from the group consisting of (1) tetramethylammonium fluoride tetrahydrate, (2) tetraethylammonium acetate tetrahydrate, (3) tetrabutylammonium chloride, (4) tetrabutylammonium chloride hydrate, (5) tetrabutylammonium bromide, (6) tetrabutylammonium tribromide, (7) tetrabutylammonium acetate, (8) tetrabutylammonium thiocyanate, (9) tetrapentylammonium bromide, (10) tetrahexylammonium bromide, (11) tetrahexylammonium chloride, (12) tetrahexylammonium hydrogensulfate, (13) tetraheptylammonium chloride, (14) tetraheptylammonium bromide, (15) tetraoctylammonium bromide, (16) tetrakisdecylammonium bromide, (17) tetrahexadecylammonium bromide, (18) tetramethyl ammonium bromide, (19) tetramethyl ammonium chloride, (20) tetramethyl ammonium iodide, (21) tetraethyl ammonium bromide, (22) tetraethyl ammonium chloride, (23) tetraethyl ammonium iodide, (24) tetrapropyl ammonium bromide, (25) tetrapropyl ammonium iodide, (26) tetrabutyl ammonium iodide, (27) tetrapentyl ammonium chloride, (28) tetrahexyl ammonium bromide, (29) tetrahexyl ammonium iodide, (30) tetradecyl ammonium bromide, (31) tetradodecyl ammonium bromide, (32) tetraoctadecyl ammonium bromide, (33) methyltrioctylammonium bromide, (34) tridodecylmethylammonium chloride, (35) tridodeylmethylammonium iodide, (36) N-dodecyl-N-methylephedrinium bromide, (37) phenyltrimethylammonium tribromide, (38) tricapryl methyl ammonium chloride, (39) tridodecyl methyl ammonium chloride, (40) tridecyloxypropyl dihydroxy ethyl methyl ammonium chloride, (41) N-tetradecyl dimethyl-naphthyl methyl ammonium chloride, (42) octadecyl diethanol methyl ammonium chloride, (43) octadecyl dihydroxyethyl methyl ammonium chloride, (44) dihydrogenated tallow benzyl methyl ammonium chloride, (45) 2-aminoethyl trimethyl ammonium chloride hydrochloride, (46) 2-bromoethyl trimethyl ammonium bromide, (47) 2-chloroethyl trimethyl ammonium chloride, (48) 3-carboxypropyl trimethyl ammonium chloride, (49) [3-(methacryloyl amino) propyl] trimethyl ammonium chloride, (50) phenyl trimethyl ammonium bromide, (51) phenyl trimethyl ammonium chloride, (52) phenyl trimethyl ammonium iodide, (53) benzyl trimethyl ammonium chloride, (54) benzyl trimethyl ammonium bromide, (55) 4-nitrobenzyl trimethyl ammonium chloride, (56) [2-(4-nitrophenyl) allyl] trimethyl ammonium iodide, (57) coco trimethyl ammonium chloride, (58) palmityl trimethyl ammonium chloride, (59) myristyl trimethyl ammonium bromide, (60) oleyl trimethyl ammonium chloride, (61) soya trimethyl ammonium chloride, (62) tallow trimethyl ammonium chloride, (63) hydrogenated tallow trimethyl ammonium chloride, (64) stearyl trimethyl ammonium chloride, (365) behenyl trimethyl ammonium chloride, (66) guar hydroxypropyl trimethyl ammonium chloride, (67) benzyl triethyl ammonium bromide, (68) butyl tripropyl ammonium bromide, (69) methyl tributyl ammonium chloride, (70) methyl tributyl ammonium bromide, (71) methyl tributyl ammonium iodide, (72) benzyl tributyl ammonium chloride, (73) benzyl tributyl ammonium bromide, (74) benzyl tributyl ammonium iodide, (75) heptyl tributyl ammonium bromide, (76) benzyldodecyldimethylammonium bromide, (77) benzyltetradecyldimethylammonium chloride dihydrate, (78) benzylcetyldimethylammonium chloride monohydrate, (79) benzylstearyldimethylammonium chloride monohydrate, (80) N,N-dimethyl methylene ammonium chloride, (81) N,N-dimethyl methylene ammonium iodide, (82) chloromethylene dimethyl ammonium chloride, (83) dichloromethylene dimethyl ammonium chloride, (84) dimethyl amino methylene amino methylene dimethyl ammonium chloride, (85) benzethonium chloride, (86) methyl benzethoniumchloride, (87) 1-propanaminium 2,3-dihydroxy-N-dimethyl-N-[3(oxococoyl) amino]propyl]-chloride, (88) cetyl dimethyl ethyl ammonium bromide, (89) octyl dodecyl dimethyl ammonium chloride, (90) dodecyl (2-hydroxy-1-methyl-2-phenyl-ethyl) dimethyl ammonium bromide, (91) dodecyl dimethyl 2-phenoxyethyl ammonium bromide, (92) dodecanoyl-N-methylamino ethyl-(phenyl carbamyl methyl) dimethyl ammonium chloride, (93) 3-chloro-2-hydroxypropyl N,N,N-dimethyl dodecyl ammonium chloride, (94) 3-chloro-2-hydroxypropyl N,N,N-dimethyl octadecyl ammonium chloride, (95) dodecyl benzyl dimethyl ammonium bromide, (96) dodecyl benzyl dimethyl ammonium chloride, (97) coco benzyl dimethyl ammonium chloride, (98) benzyl tetradecyl dimethyl ammonium chloride, (99) benzyl cetyl dimethyl ammonium chloride, (100) benzyl octadecyl dimethyl ammonium chloride, (101) benzyl tallow dimethyl ammonium chloride, (102) benzyl hydrogenated tallow dimethyl ammonium chloride, (103) benzyl behenyl dimethyl ammonium chloride, (104) dioctyl dimethyl ammonium chloride, (105) didecyl dimethyl ammonium chloride, (106) didecyl dimethyl ammonium bromide, (107) dicoco dimethyl ammonium chloride, (108) dicetyl dimethyl ammonium chloride, (109) disoya dimethyl ammonium chloride, (110) ditallow dimethyl ammonium chloride, (111) dihydrogenated tallow dimethyl ammonium chloride, (112) dibehenyl/diarachidyl dimethyl ammonium chloride, (113) soya amido propyl benzyl dimethyl ammonium chloride, (114) soya dicoco quaternary ammonium chloride, (115) gluconamidopropyl dimethyl-2-hydroxyethyl ammonium chloride, (116) N-alkyl-N-N-dimethyl-N(dodecyl acetate) ammonium chloride, wherein alkyl has from 14 to 20 carbon atoms, (117) mink amidopropyl dimethyl-2-hydroxyethyl ammonium chloride, (118) N-rapeseed-(3-amidopropyl)-N-N-dimethyl-N-(2,3 epoxy propyl) ammonium chloride, (119) N-stearyl-(3-amido propyl)-N-benzyl dimethyl ammonium chloride, (120) rapeseed amido propyl benzyl dimethyl ammonium chloride, (121) rapeseed amido propyl ethyl dimethyl ammonium chloride, (122) cocamidopropyl polyethylene glycol dimethyl ammonium chloride phosphate, (123) butyrylcholine chloride, and (124) mixtures thereof; or wherein the transparentizing agent is selected from the group consisting of piperidine thiocyanate, 2-piperidine methanol, bis(pentamethylene) urea, 4,4'-trimethylene bis(1-piperidine propionitrile), tripiperidino phosphine oxide, homopiperazine, 1-piperonyl piperazine, hexacyclentrisulfate, 5,10,15,20-tetraphenyl-21H,23Hporphine, 5,10,15,20-tetrakis(4-methoxyphenyl)-2H,23H-porphine, pyrrole-2-carboxaldehyde, 3-pyrrolidino-1,2-propanediol, pyrazole, 3-aminopyrazole, imidazole, 2-ethylimidazole, 2-(2-piperidinoethyl) pyridine, 1-dodecyl pyridinium chloride, pyridinium bromide perbromide, 3-aminoquinoline, 8-hydroxyquinoline, 7,8-benzoquinoline, 8-hydroxyquinaldine, quinoxaline, 4,5-dihydro-6-methyl-3(2H)-pyridazinone monohydrate, phthalazine, 1,10-phenanthroline, 1,3,5-triazine, trichloromelamine, trichloroisocyanouric acid, norbornane, tricyclo[5.2.1.0] decane, norcamphor, tropolone, 1-indanol, trans,trans,cis-1,5,9-cyclododecatriene, cyclodecane epoxide, 2,3-cyclododecane pyridine, 1,2,5,6,9,10-hexabromo-cyclododecane, 1,4,4a,8a-tetrahydro-endo-1,4-methano-naphthalene-5,8-dione, γ-butyrolactone, β,β-dimethyl-γ-(hydroxymethyl)-γ-butyrolactone, 2,5-dimethyl-4-hydroxy-3(2H)-furanone, hydrindantin dihydrate, 2,4,8,10-tetraoxaspiro [5.5]undecane, 1,3,5-trioxane, cyclooctanone, piperonal, piperonylalcohol, piperonyl nitrile, 3,4(methylenedioxy) phenylacetonitrile, maleic anhydride, s-acetylmercapto succinic anhydride, 2-octadecen-1-yl succinic anhydride, 18-crown-6, benzo-18 crown-6, dibenzo-18 crown-6, dibenzo-24 crown-8, 5-amino-3-methyl isooxazole, 2-oxazolidone, 5,5-dimethyl oxazolidine-2,4-dione, 3-ethyl-2-thioxo-4-oxazolidinone, 3-morpholino-1,2-propandiol, 4-phenyl morpholine, N,N'-dibenzyl-1,4,10,13- tetraoxa-7,16 diazacycloocta-decane, 4,7,13,16,21,24-hexaoxa-1,10-diazabicyclo [8.8.8] hexacosane, γ-valerolactam, ε-caprolactam, 2-azacyclooctanone, 2-azacyclononanone, maleimide, n-methylsuccinimide, phthalimide DBU salt, 1-allyl-2-thiourea, 1,3-dithiane, 1-benzyl-3-methyl-2-2-imino-4-thiobiuret, butyl sulfone, 2,2'-bithiophene, 2-phenyl-1,3-dithiane, 3,6,9,14-tetrathiabicyclo [9.2.1] tetradeca-11,13-diene, 1,5,9,13-tetra-thiacyclohexadecane-3,11-diol, 1,4,7,10,13-penta-thiacyclopentadecane, 2-aminothiazole, 2-amino-2-thiazoline, 3-methyl rhodanine, 3-ethyl-5-(2-hydroxy-ethyl)-4-methylthiazolium bromide, triphenylphosphine, tricyclohexylphosphine, 1,3-bis (diphenylphosphino) propane, 1,5-bis(diphenyl phosphino) pentane, isopropyldiphenyl phosphine, triethyl phosphite, triphenyl phosphite, triethyl phosphite copper iodide, dipropyl phosphite, bis(2-ethylhexyl) phosphite, bis(4-nitrobenzyl) phosphite, diphenyl phosphine oxide, diphenyl(2,4,6-trimethylbenzoyl) phosphine oxide, vinyl phosphonic acid, cyanoaceto-hydrazide, cyanomethyl N,N-dimethyl dithiocarbamate, 4'-pentyl-4'-biphenyl carbonitrile, 4'-(octyloxy)-4-biphenyl carbonitrile, 1,4-dicyano-2-butene, benzylidene malononitrile, 1-isothiocyanato-4-(trans-4-propylcyclohexyl)benzene, formamidoxime, ethyl chlorooximido acetate, acetohydroxamic acid, tetrahexylammonium chloride, tetraheptylammonium chloride, tetraheptylammonium bromide, and mixtures thereof.

9. A process which comprises (1) providing the migration imaging member according to claim 1, comprising (a) a substrate, (b) a softenable layer comprising a softenable material and a photosensitive migration marking material, and (c) a transparentizing agent which transparentizes migration marking material in contact therewith contained in at least one layer of the migration imaging member; (2) uniformly charging the imaging member; (3) subsequent to step (2), exposing the charged imaging member to activating radiation at a wavelength to which the migration marking material is sensitive; (4) subsequent to step (3), causing the softenable material to soften and enabling a first portion of the migration marking material to migrate through the softenable material toward the substrate in an imagewise pattern while a second portion of the migration marking material remains substantially unmigrated within the softenable layer, wherein subsequent to migration of the first portion of migration marking material, either (a) the first portion of migration marking material contacts the transparentizing agent and the second portion of migration marking material does not contact the transparentizing agent; or (b) the second portion of migration marking material contacts the transparentizing agent and the first portion of migration marking material does not contact the transparentizing agent.

10. A process according to claim 9 wherein the first portion of migration marking material contacts the transparentizing agent and the second portion of migration marking material does not contact the transparentizing agent; or wherein the second portion of migration marking material contacts the transparentizing agent and the first portion of migration marking material does not contact the transparentizing agent.

## Patentansprüche

1. Ein Migrationsbilderzeugungselement (1) umfassend (a) ein Substrat (2), (b) eine erweichbare Schicht (6) umfassend ein erweichbares Material (7) und ein photo-empfindliches Migrationsmarkierungsmaterial (8), und (c) ein transparentmachendes Mittel, welches das damit in Kontakt befindliche Migrationsmarkierungsmaterial transparent macht, enthaltend in mindestens einer Schicht des Migrationsbilderzeugungselementes, worin das transparentmachende Mittel das damit in Kontakt kommende Migrationsmarkierungsmaterial beeinflußt durch Verringern der optischen Dichte der erweichbaren Schicht, welche das Migrationsmarkierungsmaterial enthält.

2. Ein Migrationsbilderzeugungselement gemäß Anspruch 1, worin das Migrationsmarkierungsmaterial (8) ausgewählt ist aus der Gruppe bestehend aus (a) Selen, (b) Tellur, (c) Legierungen von Selen und einem Material, ausgewählt aus der Gruppe bestehend aus Tellur, Arsen, Antimon, Thallium, Wismut oder Mischungen davon, (d) Legierungen von Tellur und einem Material ausgewählt aus der Gruppe bestehend aus Arsen, Antimon, Thallium, Wismut oder Mischungen davon, (e) Halogen-dotiertem Selen, (f) Halogen-dotiertem Tellur, (g) Halogen-dotierten Legierungen von Selen und einem Material ausgewählt aus der Gruppe bestehend aus Tellur, Arsen, Antimon, Thallium, Wismut oder Mischungen davon, (h) Halogen-dotierten Legierungen von Tellur und einem Material ausgewählt aus der Gruppe bestehend aus Arsen, Antimon, Thallium, Wismut oder Mischungen davon und (i) Mischungen davon.

3. Ein Migrationsbilderzeugungselement gemäß Anspruch 1 oder Anspruch 2, worin das transparentmachende Mittel in der erweichbaren Schicht enthalten ist.

4. Ein Migrationsbilderzeugungselement gemäß Anspruch 1 oder Anspruch 2, worin das transparentmachende Mittel in einer Schicht enthalten ist, die zwischen der erweichbaren Schicht und dem Substrat angeordnet ist.

5. Das Migrationsbilderzeugungselement gemäß Anspruch 1 oder 2, worin die erweichbare Schicht zwischen dem Substrat und einer Schicht angeordnet ist, welche das transparentmachende Mittel enthält.

6. Ein Migrationsbilderzeugungselement gemäß Anspruch 1 oder Anspruch 2, worin das Migrationsbilderzeugungselement umfaßt ein Substrat, eine erste erweichbare Schicht umfassend ein erstes erweichbares Material und ein erstes Migrationsmarkierungsmaterial, und eine zweite erweichbare Schicht umfassend ein zweites erweichbares Material und ein zweites Migrationsmarkierungsmaterial, worin das transparentmachende Mittel in einer Schicht enthalten ist, die zwischen der ersten erweichbaren Schicht und der zweiten erweichbaren Schicht angeordnet ist.

7. Ein Migrationsbilderzeugungselement gemäß einem der Ansprüche 1 bis 6, worin das transparentmachende Mittel in einer Menge von etwa 1 bis etwa 50 Gew.-% des Materials umfassend die Schicht, in welcher es enthalten ist, vorhanden ist.

8. Ein Migrationsbilderzeugungselement gemäß Anspruch 1, worin das transparentmachende Mittel eine azacyclische Verbindung ist; oder worin das transparentmachende Mittel ausgewählt ist aus der Gruppe bestehend aus: (A) Materialien der allgemeinen Formeln: worin R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈ und R₃₉ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongnuppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈ und R₃₉ miteinander verbunden sein können, um einen Ring zu bilden; (B) Materialien der allgemeinen Formeln: worin R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ und R₂₂ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ und R₂₂ miteinander verbunden sein können, um einen Ring zu bilden; (C) Materialien der allgemeinen Formeln: worin R₁, R₂ und R₃ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂ und R₃ miteinander verbunden sein können, um einen Ring zu bilden; (D) Materialien der allgemeinen Formeln: worin R₁, R₂, R₃, R₄, R₅, R₆, R₇, R₈, R₉, R₁₀, R₁₁ und R₁₂ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁ und R₁₂ miteinander verbunden sein können, um einen Ring zu bilden; (E) Materialien der allgemeinen Formeln: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (F) Materialien der allgemeinen Formel: worin R₁, R₂, R₃, R₄, R₅, R₆, R₇, R₈, R₉, R₁₀, R₁₁, R₁₂, R₁₃ und R₁₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃ und R₁₄ miteinander verbunden sein können, um einen Ring zu bilden; (G) Materialien der allgemeinen Formel: worin R₁ und R₂ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin R₁ und R₂ miteinander verbunden sein können, um einen Ring zu bilden; (H) Materialien der allgemeinen Formel: worin R₁, R₂, R₃, R₄ und R₅ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄ und R₅ miteinander verbunden sein können, um einen Ring zu bilden; (1) Materialien der allgemeinen Formel: worin R₁, R₂, R₃, R_{4,} R₅, R₆, R₇, R₈ und R₉ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈ und R₉ miteinander verbunden sein können, um einen Ring zu bilden; (J) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (K) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (L) Materialien der allgemeinen Formel: worin R₁, R₂, R₃, R₄ und R₅ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄ und R₅ miteinander verbunden sein können, um einen Ring zu bilden; (M) Materialien der allgemeinen Formeln: worin R₁, R₂, R₃, R₄, R₅, R₆, R₇, R₈, R₉, R₁₀, R₁₁, R₁₂, R₁₃ und R₁₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃ und R₁₄ miteinander verbunden sein können, um einen Ring zu bilden; (N) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (O) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (P) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (Q) Materialien der allgemeinen Formel: worin R₁, R₂, R₃ und R₄ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangnuppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃ und R₄ miteinander verbunden sein können, um einen Ring zu bilden; (R) Materialien der allgemeinen Formeln: worin R₁ ausgewählt ist aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, und worin der gekrümmte Teil der Struktur eine Kohlenwasserstoffkette oder eine substituierte Kohlenwasserstoffkette bedeutet, worin zwei oder mehr Substituenten miteinander verbunden sein können, um einen Ring zu bilden; (S) Materialien der allgemeinen Formel: worin R₁ ausgewählt ist aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, und worin der gekrümmte Teil der Struktur eine Kohlenwasserstoffkette oder eine substituierte Kohlenwasserstoffkette bedeutet, worin zwei oder mehr Substituenten miteinander verbunden sein können, um einen Ring zu bilden; und (T) Mischungen davon; oder worin das transparentmachende Mittel ausgewählt ist aus der Gruppe bestehend aus (1) Homopiperidin, (2) Piperidinthiocyanat, (3) 2-Piperidinmethanol, (4) 3-Piperidinmethanol, (5) 2-Piperidinethanol, (6) 4-Piperidinethanol, (7) 4-Piperidin-Monohydrat-Hydrochlorid, (8) 1-Aminopiperidin, (9) 1-(2-Aminoethyl)piperidin, (10) 4-(Aminomethyl)piperidin, (11) 3-Piperidino-1,2-propandiol, (12) 1-Piperidinpropionsäure, (13) 1-Methyl-4-(methylamino)piperidin, (14) 1-Acetyl-3-methylpiperidin, (15) 4'-Piperidinoacetophenon, (16) 4-Phenylpiperidin, (17) 4-Piperidinopiperidin, (18) 4-Benzylpiperidin, (19) 4-(4-Methylpiperidino)pyridin, (20) 4-Piperidonethylenketal, (21) Bis(pentamethylen)harnstoff, (22) 1-Benzyl-4-hydroxypiperidin, (23) 1-Benzoyl-4-piperidon, (24)1,1'-Methylenbis(3-methylpiperidin), (25) 4,4'-Trimethylendipiperidin, (26) 4,4'-Trimethylenbis(1-menthylpiperidin), (27) 4,4'-Trimethylenbis(1-piperidinpropionitril), (28) 4,4'-Trimethylenbis(1-piperidinethanol), (29) 2,2,6,6-Tetramethylpiperidin, (30) 4-Amino-2,2,6,6-tetramethylpiperidin, (31) 4-(Dimethylamino)-1,2,2,6,6-pentamethylpiperidin, (32) N,N'-Bis(2,2,6,6-tetramethyl-4-piperidinyl)-1,6-hexandiamin, (33) Tripiperidinophosphinoxid, (34) Tropan, (35) Tropinhydrat, (36) Tropinon, (37) 8-Hydroxytropinon, (38) 2-Piperidincarbonsäure, (39) 2-Piperidon, (40) 4,4'-Trimethylenbis(1-piperidincarboxamid), (41) 4-Methyl-2-(piperidinomethyl)phenol, (42) 1-Methyl-4-piperidinylbis(chlorphenoxy)acetat, (43) 2-(Hexamethylenimino)ethylchlorid-Monohydrochlorid, (44) 3-(Hexahydro-1H-azepin-1-yl)-3'-nitropropiophenon-Hydrochlorid, (45) lmipramin-Hydrochlorid, (46) Carbamezepin, (47) 5,6,11,12-Tetrahydrodibenz[b,f]azocin-Hydrochlorid, (48) Chinuclidin-Hydrochlorid, (49) 3-Chinuclidinol-Hydrochlorid, (50) 3-Chinuclidinon-Hydrochlorid, (51) 2-Methylen-3-chinuclidinon-Dihydrat-Hydrochlorid, (52) 3-Aminochinuclidin-Dihydrochlorid, (53) 3-Chlorchinuclidin-Hydrochlorid, (54) Chinidinsulfat-Dihydrat, (55) Chinin-Monohydrochlorid-Dihydrat, (56) Chininsulfat-Monohydrat, (57) Hydrochinidin-Hydrochlorid, (58) Hydrochinin-Hydrobromid-Dihydrat, (59) Piperazin, (60) Homopiperazin, (61) 1-Methylpiperazin, (62) 2-Methylpiperazin, (63) 1-Acetylpiperazin, (64) 1-(2-Hydroxyethyl)piperazin, (65) 1-(2-Aminoethyl)piperazin, (66) tert-Butyl-1-piperazincarboxylat, (67) N-lsopropyl-1-piperazinacetamid, (68) 1-(2-Methoxyphenyl)piperazin, (69) 1-(2-Pyridyl)piperazin, (70) 1-Benzylpiperazin, (71) 1-Cinnamylpiperazin, (72) 1-(4-Chlorbenzhydryl)piperazin, (73) 2,6-Dimethylpiperazin, (74) 1-Amino-4-methylpiperazin, (75) 1-Amino-4-(2-hydroxyethyl)piperazin, (76) 1,4-Bis(2-hydroxyethyl)piperazin, (77) 1,4-Bis(3-aminopropyl)piperazin, (78) tert-Butyl-4-benzyl-1-piperazincarboxylat, (79) 1-Piperonylpiperazin, (80) Bis(4-methyl-1-homopiperazinylthiocarbonyl)disulfid, (81) 1-Amino-4-methylpiperazin-Dihydrochlorid-Monohydrat, (82) 1-(3-Chlorpropyl)piperazin-Dihydrochlorid-Monohydrat, (83) 1-(2,3-Xylyl)piperazin-Monohydrochlorid, (84) 1,1-Dimethyl-4-phenylpiperaziniumiodid, (85) 1,4,7-Triazacyclononan, (86) 1,5,9-Triazacyclododecan, (87) 1,2,3-Triazol, (88) 4-Amino-1,2,4-triazol, (89) 3-Amino-5-methylthio-1H-1,2,4-triazol, (90) Benzotriazol, (91) 1-Aminobenzotriazol, (92) 1-Cyanbenzotriazol, (93) 5-Methyl-1 H-benzotriazol, (94) 1 H-Benzotriazol-1-ylmethylisocyanid, (95) 2-[3-(2H-Benzotriazol-2-yl)-4-hydroxyphenyl] ethylmethacrylat, (96) 1,2,4-Triazol, (97) 1,2,4-Triazol-Natriumderivat, (98) 3-Amino-1,2,4-triazol, (99) 3,5-Diamino-1,2,4-triazol, (100) 3-Amino-5-mercapto-1,2,4-triazol, (101) 3-Amino-1,2,4-triazol-5-carbonsäure-Hemihydrat, (102) 4-Amino-3-hydrazino-5-mercapto-1,2,4-triazol, (103) 1,2,3-Triazol-4,5-dicarbonsäure-Monohydrat, (104) Nitron, (105) 1-Hydroxybenzotriazol-Hydrat, (106) 1,3,5-Triazin, (107) Cyanursäure, (108) Trithiocyanursäure, (109) 2,4-Bis(methylthio)-6-chlor-1,3,5-triazin, (110) 2-Chlor-4,6-dimethoxy-1,3,5-triazin, (111) 2-Chlor-4,6-diamino-1,3,5-triazin, (112) Trichlormelamin, (113) Cyanurchlorid, (114) 2,4,6-Tris(perfluorheptyl)-1,3,5-triazin, (115) Hexahydro-2,4,6-trimethyl-1,3,5-triazin-Trihydrat, (116) 1,3,5-Trimethylhexahydro-1,3,5-triazin, (117) 1,3,5-Triethylhexahydro-1,3,5-triazin, (118) 1,3,5-Triclohexylhexahydro-1,3,5-triazin, (119) 1,3,5-Tribenzylhexahydro-1,3,5-triazin, (120) Trichlorisocyanursäure, (121) Tris(2,3-dibrompropylisocyanurat), (122) Cyanursäureverbindung mit Melamin, (123) Urazol, (124) 1-Methylurazol, (125) 4-Phenylurazol, (126) 5-(4-Hydroxyphenyl)-5-phenylhydantoin, (127) β-Tetralonhydantoin, (128) Cyclen (1,4,7,10-Tetraazacyclododecan), (129)1,4,8,11-Tetraazacyclotetradecan, (130)1,4,8,11-Tetramethyl-1,4,8,11-tetraazacyclotetradecan, (131) 1,4,8,11-Tetraazacyclotetradecan-5,7-dion, (132) 1,4,8,12-Tetraazacyclopentadecan, (133) 2,3,7,8,12,13,17,18-Octaethyl-21H,23H-porphin, (134) Dimethyl-3,7,12,17-tetramethyl-21H,23H-porphin-2,18-dipropionat, (135) Dimethyl-7,12-diacetyl-3,8,13,17-tetramethyl-21 H,23H-porphin-2,18-dipropionat, (136) 8,3-Divinyl-3,7,12,17-tetramethyl-21 H,23H-porphin-2,18-dipropionsäure, Dinatriumsalz, (137) 5,10,15,20-Tetraphenyl-21H,23H-porphin, (138) 5,10,15,20-Tetrakis(4-methoxyphenyl)-21H,23H-porphin, (139) 5,10,15,20-Tetrakis[4-(trimethylamino)phenyl]-21H,23H-porphin, Tetra-p-tosylatsalz , (140) 5,10,15,20-Tetra(4-pyridyl)-21H,23H-porphin, (141) 5,10,15,20-Tetrakis(1-methyl-4-pyridyl)-21H,23H-porphin, Tetra-p-tosylatsalz, (142) 1,5-Pentamethylentetrazol, (143)1-H-Tetrazol, (144) 5-Aminotetrazol-Monohydrat, (145) 2,3,5-Triphenyl-2H-tetrazoliumchlorid, (146) 2-(4-lodphenyl)-5-(4-nitrophenyl)-3-phenyltetrazoliumchlorid, (147) 1,2,3,3-Tetramethyl-3H-indoliniumiodid, (148) Hexacyclentrisulfat, (149) Hexamethylhexacyclen, (150) Pyrrol-2-carboxaldehyd, (151) Prolinamid, (152) 3-Pyrrolidino-1,2-propandiol, (153) 1-(Pyrrolidinocarbonylmethyl)piperazin, (154) 4-Pyrrolidinopyridin, (155) 3-lndolylacetonitril, (156) 6-Nitroindolin, (157) 7-Azaindol, (158) Indazol, (159) 2-Acetylpyrrol, (160) 2-Acetyl-1-methylpyrrol, (161) 3-Acetyl-1-methylpyrrol, (162) 3-Acetyl-2,4-dimethylpyrrol, (163) Pyrrol-2-carbonsäure, (164) 3-Carboxy-1,4-dimethyl-2-pyrrolessigsäure, (165) Prolin, (166) 2-Pyrrolidon-5-carbonsäure, (167) 4-Hydroxyprolin, (168) 1,1'-Ethylenbis(5-oxo-3-pyrrolidincarbonsäure), (169) Kainsäure-Monohydrat, (170) 1-Aminopyrrolidin-Hydrochlorid, (171) 2-(2-Chlorethyl)-1-methylpyrrolidin-Hydrochlorid, (172) 1-(2-Chlorethyl)pyrrolidin-Hydrochlorid, (173) Tremorin-Dihydrochlorid, (174) L-Prolinmethylester-Hydrochlorid, (175) Ammoniumpyrrolidindithiocarbamat, (176) Pyrrolidon-Hydrotribromid, (177) 1-(4-Chlorbenzyl)-2-(1-pyrrolidinylmethyl)benzimidazol-Hydrochlorid, (178) Billverdin-Dihydrochlorid, (179) Indol, (180) 4,5,6,7-Tetrahydroindol, (181) 3-lndolmethanol-Hydrat, (182) 3-lndolethanol, (183) Indol-3-carboxaldehyd, (184) 3-lndolylacetat, (185) Indol-3-acetamid, (186) Indol-3-carbonsäure, (187) Indol-3-essigsäure, (188) 3-lndolpropionsäure, (189) 3-Indolacrylsäure, (190) 3-lndolglyoxylsäure, (191) Indol-3-pyruvinsäure, (192) 3-Indolmilchsäure, (193) 3-Indolbuttersäure, (194) N-Acetyltryptophanamid, (195) N-(3-lndolylacetyl)alanin, (196) N-(3-lndolylacetyl)valin, (197) N-(3-lndolylacetyl)isoleucin, (198) N-(3-lndolylacetyl)leucin, (199) N-(3-lndolylacetyl)asparaginsäure, (200) N-(3-lndolylacetyl)-L-phenylalanin, (201) 4-Hydroxyindol, (202) Indol-4-carbonsäure, (203) 4-lndolylacetat, (204) 4-Methylindol, (205) 5-Hydroxyindol, (206) 5-Hydroxyindol-3-essigsäure, (207) 5-Hydroxy-2-indolcarbonsäure, (208) N-Acetyl-5-hydroxytryptamin, (209) Indol-5-carbonsäure, (210) 5-Methylindol, (211) 5-Methoxyindol, (212) Indol-2-carbonsäure, (213) lndolen-2-carbonsäure, (214) Indol-2,3-dion, (215) 2-Methylindol, (216) 2,3,3-Trimethylindolenin, (217) Tryptamin-Hydrochlorid, (218) 5-Methyltryptamin-Hydrochlorid, (219) Serotonin-Hydrochlorid-Hemihydrat, (220) Norharman-Hydrochlorid-Monohydrat, (221) Harman-Hydrochlorid-Monohydrat, (222) Harmin-Hydrochlorid-Hydrat, (223) Harmalin-Hydrochlorid-Dihydrat, (224) Harmol-Hydrochlorid-Dihydrat, (225) Harmalol-Hydrochlorid-Dihydrat, (226) 3,6-Diaminoacridin-Hydrochlorid, (227) (3-lndolyl)isothiuroniumiodid, (228) Yohimbin-Hydrochlorid, (229) Pyrazol, (230) 3-Aminopyrazol, (231) 5-Amino-1-ethylpyrazol, (232) 3-Amino-4-carbethoxypyrazol, (233) 3-Amino-5-methylpyrazol, (234) 3-Amino-5-phenylpyrazol, (235) Ethyl-4-pyrazolcarboxylat, (236) Diethyl-3,5-pyrazolcarboxylat, (237) 1,1'-(1-Ethylpropyliden)bis-1H-pyrazol, (238) 4-Brompyrazol, (239) 4-Brom-3-methylpyrazol, (240) 3,5-Dimethylpyrazol, (241) 4-Brom-3,5-dimethylpyrazol, (242) 3,5-Dimethylpyrazol-1-carboxamid, (243) 3,5-Dimethylpyrazol-1-methanol, (244) 3-Methyl-1-vinylpyrazol, (245) 4-Benzoyl-3-methyl-1-phenyl-2-pyrazolin-5-on, (246) 1-Nitropyrazol, (247) 4-Pyrazolcarbonsäure, (248) 3,5-Pyrazoldicarbonsäure-Monohydrat, (249) 3-Amino-5-hydroxypyrazol, (250) 3-Amino-4-pyrazolcarbonitril, (251) 3-Amino-4-pyrazolcarbonsäure, (252) 4-Methylpyrazol-Hydrochlorid, (253) 3,4-Diamino-5-hydroxypyrazolsulfat, (254) 3,5-Dimethylpyrazol-1-carboxamidinnitrat, (255) 3-Amino-4-pyrazolcarboxamid-Hemisulfat, (256) Säuresalz von 6-Aminoindazol-Hydrochlorid, (257) 4-Hydroxypyrazolo-[3,4-d]-pyrimidin, (258) 4-Mercapto-1 H-pyrazolo-[3,4-d]-pyrimidin, (259) Indazol, (260) 5-Aminoindazol, (261) 6-Aminoindazol, (262) 3-Indazolinon, (263) N'-(6-Indazolyl)sulfanilamid, (264) 4,5-Dihydro-3-(4-pyridinyl)-2H-benz[g]indazol-Methansulfonat, (265) Imidazol, (266) 4-Methylimidazol, (267) 2-Ethylimidazol, (268) 2-Propylimidazol, (269) 1-Butylimidazol, (270) 2-Undecylimidazol, (271) Histamin, (272) 1-(3-Aminopropyl)imidazol, (273) 1-Acetylimidazol, (274) 2-Methyl-1-vinylimidazol, (275) 2-Ethyl-4-methylimidazol, (276) 1-Benzyl-2-methylimidazol, (277) 1-Methylbenzimidazol, (278) 1-Ethyl-3-methyl-1,H-imidazoliniumchlorid, (279) 2-(Aminomethyl)benzimidazol-Dihydrochlorid-Hydrat, (280) 2,6-Diamino-8-purinol-Hemisulfat-Monohydrat, (281) Purin-6-yl-trimethylammoniumchlorid, (282) 4-Methyl-5-imidazolmethanol-Hydrochlorid, (283) N,N'-Bis[3-(4,5-dihydro-1H-imidazol-2-yl)phenyl]harnstoffdipropanoat, (284) 1-(p-Tosyl)-3,4,4-trimethyl-2-imidazoliniumiodid, (285) 1-Ethyl-3-methyl-1 H-imidazoliniumchlorid, (286) 2-Aminoimidazolsulfat, (287) 4-Amino-5-imidazolcarboxamid-Hydrochlorid, (288) 2-Hydrazino-2-imidazolin-Hydrobromid, (289) Imidazol-Hydrochlorid, (290) 4-lmidazolessigsäure-Hydrochlorid, (291) 2-Benzyl-2-imidazolin-Hydrochlorid, (292) Propyl-1-(1-phenylethylimidazol-5-carboxylat-Hydrochlorid, (293) 2,6-Diaminopurinsulfat-Hydrat, (294) 1-Talgamidoethyl-3-methyl-2-heptadecylimidazolinium-Methylsulfat, (295) Isostearylethylimidonium-Ethylsulfat, (296) Methyl-(1)-talgamidoethyl-2-talgimidazolinium-Methylsulfat, (297) Isostearylbenzylimidoniumchlorid, (298) Methyl-(1)-hydriertes Talgamidoethyl, (299) hydriertes Talgimidazolinium-Methylsulfat, (300) 1-Methyl-1-oleylamidoethyl-2-oleylimidazolinium-Methylsulfat, (301) Kokoshydroxyethylpolyethylenglycolimidazoliniumchloridphosphat, (302) Guanin, (303) Guanosin-Hydrat, (304) Xanthin, (305) 1-Methylxanthin, (306) 3-Methylxanthin, (307) 3-lsobutyl-1-methylxanthin, (308) Hypoxanthin, (309) Xanthosin-Dihydrat, (310) 6-Thioxanthen, (311) Purin, (312) 6-Aminopurin, (313) 6-Methoxypurin-Hemihydrat, (314) 6-Mercaptopurin-Monohydrat, (315) 2-Amino-6-chlorpurin, (316) 2-Amino-6,8-dihydroxypurin, (317) Theophyllin (3,7-Dihydro-1,3-dimethyl-1H-purin-2,6-dion), (318) Kinetin (6-Furfurylaminopurin), (319) 1-Methyladenin, (320) 3-Methyladenin, (321) Adenosin, (322) Inosin, (323) 6-Mercaptopurinribosid, (324) 6-Aminopurin-Hydrochlorid-Hemihydrat, (325) 6-Aminopurinsulfat, (326) 2,6-Diamino-8-purinol-Hemisulfat-Monohydrat, (327) Benzimidazol, (328) 2-Aminobenzimidazol, (329) 2-Amino-5,6-dimethylbenzimidazol, (330) 5-Benzimidazolcarbonsäure, (331) 2,4,5-Trimethylbenzimidazol, (332) 2-Guanidinobenzimidazol, (333) 2-Hydroxybenzimidazol, (334) 4-(2-Keto-1-benzimidazolinyl)piperidin, (335) 2-lmidazolidinthion, (336) 2-lmidazolidon, (337) Hydantoin, (338) 1-Methylhydantoin, (339) Kreatinin, (340) 2-Thiohydrantoin, (341) 5-Hydantoinessigsäure, (342) 5-Ureidohydantoin, (343) 5,5-Dimethylhydantoin, (344) 2-lmidazolidon-4-carbonsäure, (345) N,N-Bis(2-hydroxyethyl)isonicotinamid, (346) 1,2-Bis(4-pyridyl)ethylen, (347) 2-(2-Piperidinoethyl)pyridin, (348) 1,2-Bis(4-pyridyl)ethan, (349) 4,4'-Trimethylenpyridin, (350) Aldrithiol-2, (351) Aldrithiol-4, (352) 1,3-Bis(3-pyridylmethyl)-2-thioharnstoff, (353) 2,2':6',2"-Terpyridin, (354) 2-[N,N-Bis(trifluormethylsulfonyl)amino]pyridin, (355) 2,3-Pyridindicarbonsäure, (356) 2,4-Pyridindicarbonsäure-Monohydrat, (357) 2,5-Pyridindicarbonsäure, (358) 2,6-Pyridindicarbonsäure, (359) 3,4-Pyridindicarbonsäure, (360) 3,5-Pyridindicarbonsäure, (361) 2,6-Pyridindicarboxaldehyd, (362) 3,4-Pyridincarboxamid, (363) 3,4-Pyridincarboximid, (364) 2,3-Pyridincarbonsäureanhydrid, (365) 3,4-Pyridincarbonsäureanhydrid, (366) 2,6-Pyridinmethanol, (367) 2-Pyridinethansulfonsäure, (368) 4-Pyridinethansulfonsäure, (369) 3-Pyridinsulfonsäure, (370) Pyridoxsäure, (371) trans-3-(3-Pyridyl)acrylsäure, (372) 2-Pyridylhydroxymethansulfonsäure, (373) 3-Pyridylhydroxymethansulfonsäure, (374) 6-Methyl-2,3-pyridindicarbonsäure, (375) Isonicotinsäure, (376) Pyridin-Hydrobromid, (377) Pyridin-Hydrochlorid, (378) 2-(Chlormethyl)pyridin-Hydrochlorid, (379) 2-PyridylessigsäureHydrochlorid, (380) Nicotinoylchlorid-Hydrochlorid, (381) 2-Hydrazinopyridin-Dihydrochlorid, (382) 2-(2-Methylaminoethyl)pyridin-Dihydrochlorid, (383) 1-Methyl-1,2,3,6-tetrahydropyridin-Hydrochlorid, (384) 2,6-Dihydroxypyridin-Hydrochlorid, (385) 3-Hydroxy-2-(hydroxymethyl)pyridin-Hydrochlorid, (386) Pyridoxin-Hydrochlorid, (387) Pyridoxal-Hydrochlorid, (388) Pyridoxal-5-phosphat-Monohydrat, (389) 3-Amino-2,6-dimethoxypyridin-Hydrochlorid, (390) Pyridoxamin-Dihydrochlorid-Monohydrat, (391) Iproniazidphosphat, (392) Tripelennamin-Hydrochlorid, (393) Pyridiniumbromidperbromid, (394) Pyridinium-3-nitrobenzolsulfonat, (395) 1-Ethyl-3-hydroxypyridiniumbromid, (396) 1-Ethyl-4-(methoxycarbonyl)pyridiniumiodid, (397) 1-Heptyl-4-(4-pyridyl)pyridiniumbromid, (398) 1-Dodecylpyridiniumchlorid, (399) 1-Hexadecylpyridiniumchlorid-Monohydrat, (400) 1-Hexadecylpyridiniumbromid-Monohydrat, (401) 1-(Carboxymethyl)pyridiniumchlorid, (402) 1-(Carboxymethyl)pyridiniumchloridhydrazid, (403) 1-(3-Nitrobenzyloxymethyl)pyridiniumchlorid, (404) 1-(3-Sulfopropyl)pyridiniumhydroxid, (405) N-(Lauroylcolaminoformylmethyl)pyridiniumchlorid, (406) N-(Stearoylcolaminformylmethyl)pyridiniumchlorid, (407) 2-Chlor-1-methylpyridiniumiodid, (408) 2-Pyridinaldoxim-1-methylmethansulfonat, 2-Pyridinaldoxim-1-methylchlorid, (409) 2-[4-(Dimethylamino)styryl]-1-ethylpyridiniumiodid, (410) 1-Benzyl-3-hydroxypyridiniumchlorid, (411) 1,4-Dimethylpyridiniumiodid, (412) 1-Ethyl-4-phenylpyridiniumiodid, (413) 4-Phenyl-1-propylpyridiniumiodid, (414) 1-Docosyl-4-(4-hydroxystyryl)pyridiniumbromid, (415) 1,1'-Dimethyl-4-4'-bipyridiniumdichlorid, (416)1,1'-Diethyl-4-4'-bipyridiniumdibromid, (417) 1,1'-Dibenzyl-4,4'-bipyridiniumdichlorid, (418) 1,1'-Diheptyl-4,4'-bipyridiniumdibromid, (419) 1,7-Phenanthrolin, (420) 1,10-Phenanthrolin, (421) 5-Chlor-1,10-phenanthrolin, (422) 4,5-Dihydro-3-(4-pyridinyl)-2H-benz[g]indazol-Methansulfonat, (423) 1,2,3,4-Tetrahydrochinolin, (424) 6-Ethoxy-1,2,3,4-tetrahydro-2,2,4-trimethylchinolin, (425) 2-Cyanchinolin, (426) 1-Cyanisochinolin, (427) 3-Cyanisochinolin, (428) 3-Aminochinolin, (429) 8-Aminochinolin, (430) 7,8-Benzochinolin, (431) 8-Hydroxychinolin, (432) 8-Hydroxychinolin-Aluminiumsalz, (433) 8-Hydroxychinaldin, (434) 3,4,5,6,7,8-Hexahydro-2-(1H)-chinolinon, (435) Julolidin, (436) Chinoxalin, (437) Ethyl-2-chinoxalincarboxylat, (438) Chinolin, (439) 2-Hydroxychinolin, (440) 4-Hydroxychinolin, (441) 5-Hydroxychinolin, (442) 5-Aminochinolin, (443) 6-Aminochinolin, (444) 2-Chinolincarbonsäure, (445) 3-Chinolincarbonsäure, (446) 4-Chinolincarbonsäure, (447) 4-Chinolincarboxaldehyd, (448) 2-Chinolinthiol, (449) 2,4-Chinolindiol, (450) Chinaldin, (451) 4-Aminochinaldin, (452) 2,6-Dimethylchinolin, (453) 2,7-Dimethylchinolin, (454) 4-Methoxy-2-chinolincarbonsäure, (455) Methyl-2-phenyl-4-chinolincarboxylat, (456) 2-(N-Butylcarbamoyl)-1,2,3,4-tetrahydroisochinolin, (457) 1-Hydroxyisochinolin, (458) 1-lsochinolincarbonsäure, (459) 3-lsochinolincarbonsäure, (460) 1,5-lsochinolindiol, (461) 8-Hydroxychinolin-Hemisulfat-Hemihydrat, (462) 5-Amino-8-hydroxychinolin-Dihydrochlorid, (463) 2-(Chlormethyl)chinolin-Monohydrochlorid, (464) 8-Hydroxychinolin-5-sulfonsäure-Monohydrat, (465) 8-Ethoxy-5-chinolinsulfonsäure-Natriumsalz-Hydrat. (466) 1,2,3,4-Tetrahydroisochinolin-Hydrochlorid, (467) 1,2,3,4-Tetrahydro-3-isochinolincarbonsäure-Hydrochlorid, (468) 6,7-Dimethoxy-1,2,3,4-tetrahydroisochinolin-Hydrochlorid, (469) 1-Methyl-6,7-dihydroxy-1,2,3,4-tetrahydroisochinolin-Hydrobromid, (470) Primachindiphosphat, (471) Pentachinphosphat, (472) Dibucain-Hydrochlorid, (473) 9-Aminoacridin-Hydrochlorid-Hemihydrat, (474) 3,6-Diaminoacridin-Hemisulfat, (475) 2-Chinolinthiol-Hydrochlorid, (476) Sparteinsulfat-Pentahydrat, (477) Papaverin-Hydrochlorid, (478) Emetin-Dihydrochlorid-Hydrat, (479) 1,10-Phenanthrolin-Monohydrochlorid-Monohydrat, (480) Neocuproin-Hydrochlorid-Trihydrat, (481) Pyrimidin, (482) 2-Chlorpyrimidin, (483) 4-Phenylpyrimidin, (484) 5-Brompyrimidin, (485) 2,4-Dichlorpyrimidin, (486) 4,6-Dichlorpyrimidin, (487) 2,4-Dichlor-6-methylpyrimidin, (488) 6-Chlor-2,4-dimethoxypyrimidin, (489) 2-Amino-4,6-dimethoxypyrimidin, (490) 2,4,6-Trichlorpyrimidin, (491) 2,4,5,6-Tetrachlorpyrimidin, (492) 1,3,4,6,7,8-Hexahydro-1-methyl-2H-pyrimido-[1,2-a]-pyrimidin, (493) 1,3,4,6,7,8-Hexahydro-2H-pyrimido-[1,2-a]-pyrimidin, (494) Hexetidin, (495) tert-Butyl-S-(4,6-dimethylpyrimidin-2-yl)thiocarbonat, (496) 4-MethoxybenzylS(4,6-dimethylpyrimidin-2-yl)thiocarbonat, (497) 2-Aminopyrimidin, (498) 2-Amino-4-methylpyrimidin, (499) 2-Amino-5-nitropyrimidin, (500) 2-Amino-5-brompyrimidin, (501) 2-Amino-4-chlor-6-methylpyrimidin, (502) 2-Amino-4,6-dimethylpyrimidin, (503) 2-Amino-4-hydroxy-6-methylpyrimidin, (504) 2-Amino-4,6-dichlorpyrimidin, (505) 2-Amino-5-brom-6-methyl-4-pyrimidinol, (506) 4-Aminopyrimidin, (507) 4,5-Diaminopyrimidin, (508) 4-Amino-2,6-dimethylpyrimidin, (509) 2,4-Diamino-6-hydroxypyrimidin, (510) 2,6-Diamino-4-chlorpyrimidin, (511) 4,6-Diamino-2-mercaptopyrimidin-Hemihydrat, (512) 2,4,6-Triaminopyrimidin, (513) 5-Nitroso-2,4,6-triaminopyrimidin, (514) 4,6-Dihydroxypyrimidin, (515) 4,6-Dihydroxy-2-aminopyrimidin, (516) 4,6-Dihydroxy-2-methylpyrimidin, (517) 4,6-Dihydroxy-5-nitropyrimidin, (518) 2,4-Dihydroxy-5-methylpyrimidin, (519) 2,4-Dihydroxy-6-methylpyridimin, (520) 2,4-Dihydroxy-5,6-dimethylpyrimidin, (521) 2,6-Dihydroxypyrimidin-5-carbonsäure-Hydrat, (522) 2,6-Dihydroxy-4-aminopyrimidin, (523) 2,4,5-Trihydroxypyrimidin, (524) 2-Thiouracil, (525) 6-Amino-5-nitroso-2-thiouracil, (526) Folsäure-Dihydrat, (527) Folinsäure-Calciumsalz-Hydrat, (528) 2-Hydroxypyrimidin-Hydrochlorid, (529) 2-Hydroxy-4-methylpyrimidin-Hydrochlorid, (530) 4,6-Dimethyl-2-hydroxypyrimidin-Hydrochlorid, (531) 2-Mercapto-4-methylpyrimidin-Hydrochlorid, (532) 4,6-Diaminopyrimidin-Hemisulfat-Monohydrat, (533) 4,5,6-Triaminopyrimidinsulfat-Hydrat, (534) 4,5-Diamino-6-hydroxypyrimidinsulfat, (535) 2,4-Diamino-6-mercaptopyrimidin-Hemisulfat, (536) 2,4-Diamino-6-hydroxypyrimidin-Hemisulfat-Hydrat, (537) 6-Hydroxy-2,4,5-triaminopyrimidinsulfat, (538) 5,6-Diamino-2,4-dihydroxypyrimidinsulfat, (539) N4-(2-Amino-4-pyrimidinyl)sulfanilamid-Monohydrochlorid, (540) 2,4,5,6-Tetraaminopyrimidinsulfat, (541) 2,4-(1H,3H)-Pyrimidindion, (542) 5-Aminouracil, (543) 5-Nitrouracil, (544) 5-loduracil, (545) 5-(Hydroxymethyl)uracil-Hydrat, (546) 5,6-Dihydrouracil, (547) 6-Amino-1-methyluracil, (548) 5,6-Diamino-1,3-dimethyluracil-Hydrat, (549) Uridin, (550) 5-Methyluridin, (551) 5-loduridin, (552) Thimidin, (553) 5-Methyl-2-thiouracil, (554) 4-Thiouridin, (555) 2-Thiocytidin-Dihydrat, (556) Orotsäure-Monohydrat, (557) Hydroorotsäure, (558) 5-Aminoorotsäure, (559) Methylorotat (560) Barbitursäure, (561) 5-Nitrobarbitursäure-Trihydrat, (562) Violursäure-Monohydrat, (563) Alloxan-Monohydrat, (564) 4,5,6-Triamino-2(1H)-pyrimidinthionsulfat, (565) Cyclocytidin-Hydrochlorid, (566) Cytosinarabinosid-Hydrochlorid, (567) Pyridazin, (568) Phthalazin, (569) 4,5-Dihydro-6-methyl-3(2H)-pyridazinon-Monohydrat, (570) 3,6-Dichlorpyridazin, (571) 3,4,5-Trichlorpyridazin, (572) 3,6-Dichlor-4-methylpyridazin, (573) 3-Chlor-6-methoxypyridazin, (574) Pyrazin, (575) Acetylpyrazin, (576) Aminopyrazin, (577) 2,6-Dichlorpyrazin, (578) 2,3,5-Trimethylpyrazin, (579) Tetramethylpyrazin, (580) 5-Methyl-2-pyrazincarbonsäure, (581) Pyrazinamid, (582) 2,3-Pyrazindicarboxamid, (583) 4-Pyridazincarbonsäure, (584) 2,3-Pyrazindicarbonsäure, (585) Lumazin-Monohydrat, (586) Xanthopterin-Monohydrat, (587) 2-Chinoxazolincarbonsäure, (588) 2-Chinoxalinol, (589) 2,3-Dihydroxychinoxalin, (590) Phenazinmethosulfat, (591) 2-Azetidinon, (592) 2-Pyrrolidinon, (593) Pyrrolidon-Hydrotribromid, (594) δ-Valerolactam, (595) ε-Caprolactam, (596) Amino-ε-caprolactam, (597) N-Methylcaprolactam, (598) 2-Azacyclooctanon, (599) 2-Azacyclononanon, (600) ω-Thiocaprolactam, (601) N-Vinylcaprolactam, (602) 2-Azabicyclo[2.2.1]hept-5-en-3-on, (603) Maleimid, (604) N-Ethylmaleimid, (605) N-Butylmaleimid, (606) N-Cyclohexylmaleimid, (607) N-Phenylmaleimid, (608) N-Benzylmaleimid, (609) N-Hydroxymaleimid, (610) Succinimid, (611) N-Methylsuccinimid, (612) 2-Hydroxy-N-methylsuccinimid, (613) N-Hydroxysuccinimid, (614) Succinimidyl-2,2,2-trichlorethylcarbonat, (615) 2-Dodecyl-N-(2,2,6,6-tetramethyl-4-piperidinyl)succinimid, (616) 2-Dodecy-N-(1,2,2,6,6-pentamethyl-4-piperidinyl)succinimid, (617) N-(1-Acetyl-2,2,6,6-tetramethyl-4-piperidinyl)-2-dodecylsuccinimid, (618) α-Methyl-α-propylsuccinimid, (619) α-Methyl-α-phenylsuccinimid, (620) N-Vinylphthalimid, (621) N-Ethylphthalimid, (622) N-(Trimethylsilylmethyl)phthalimid, (623) N-(2-Bromethyl)phthalimid, (624) N-(3-Brompropyl)phthalimid, (625) N-(4-Brombutyl)phthalimid, (626) Phthalimidoacetaldehyddiethylacetal, (627) Diethyl(phthalimidomethyl)phosphonat, (628) N-Benzylphthalimid, (629) Phthalimid, DBU (1,8-Diazabicyclo[5.4.0]undec-7-en)-Salz, (630) Phthalimid, DBN (1,5-Diazabicyclo[4.3.0]non-5-en), und (631) Mischungen davon; oder worin das transparentmachende Mittel eine Oxaaza-cyclische Verbindung ist, oder worin das transparentmachende Mittel ausgewählt ist aus der Gruppe bestehend aus: (A) Materialien der allgemeinen Formeln: worin R₁, R₂, R₃, R₄, R₅, R₆, R₇, R₈, R₉, R₁₀, R₁₁, R₁₂, R₁₃, R₁₄ und R₁₅ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃, R₁₄ und R₁₅ miteinander verbunden sein können, um einen Ring zu bilden; (B) Materialien der allgemeinen Formel: worin R₁, R₂, R₂, R₄, R₅, R₆, R₇, R₈ und R₉ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈ und R₉ miteinander verbunden sein können, um einen Ring zu bilden; (C) Mischungen davon; oder worin das transparentmachende Mittel ausgewählt ist aus der Gruppe bestehend aus (1) 3-Amino-5-methylisoxazol, (2) 5-Amino-3-methylisoxazol, (3) 3,5-Dimethyl-4-nitroisoxazol, (4) 1,2-Benzisoxazol, (5) 2,1-Benzisoxazol, (6) Cycloserin, (7) 4-Benzyl-2-methyl-2-oxazolin, (8) 2-Methyl-5-phenyl-2-oxazolin-4-methanol, (9) Benzoxazol, (10) 2-Methylbenzoxazol, (11) 2-Chlorbenzoxazol, (12) 2-Chlor-3-ethylbenzoloxazoliumtetrafluorborat, (13) 2-Oxazolidon, (14) 3-Methyl-2-oxazolidinon, (15) 5-Chlormethyl-2-oxazolidinon, (16) 4-lsopropyl-2-oxazolidinon, (17) 3-Acetyl-2-oxazolidinon, (18) 5,5-Dimethyloxazolidin-2,4-dion, (19) 3-Ethyl-2-thioxo-4-oxazolidinon, (20) 4-Methyl-5-phenyl-2-oxazolidinon, (21) 4-Benzyl-2-oxazolidinon, (22) 2-Benzoisoxazolinon, (23) Muscimol-Hydrat, (24) 5-Methyl-3-phenylisoxazol-4-carbonsäure, (25) 2-Methyl-5-phenyl-2-oxazolin-4-methanol, (26) Sulfamethoxazol, (27) Sulfisoxazol, (28) N'-(4,5-Dimethyloxazol-2-yl)sulfanilamid, (29) Cloroxazon, (30) 3,3'-Dimethyloxacarbocyaniniodid, (31) 2-Ethyl-5-phenylisoxazolium-3'-sulfonat, (32) 2-tert-Butyl-5-methylisoxazoliumperchlorat, (33) 5-Phenyl-2-(4-pyridyl)oxazol-Hydrochlorid-Hydrat, (34) 5-Phenyl-2-(4-pyridyl)oxazolmethyl-Tosylatsalz, (35) 4-Aminomorpholin, (36) 4-Morpholincarbonitril, (37) 4-Morpholinpropionitril, (38) 4-Formylmorpholin, (39) 4-Acetylmorpholin, (40) 4-(2-Hydroxyethyl)morpholin, (41) 3-Morpholino-1,2-propandiol, (42) 4-(3-Aminopropyl)morpholin, (43) 1-Morpholino-1-cyclopenten, (44) 1-Morpholino-1-cyclohexen, (45) 1-Morpholino-1-cyclohepten, (46) 4-Phenylmorpholin, (47) 4-Morpholinoanilin, (48) 2,2,2-Tribromethylphosphoromorpholinochloridat, (49) 1-(Morpholinocarbonylmethyl)piperazin, (50) 1,3-Dimorpholin-2-nitropropan, (51) Hemicholinium-3, (52) Hemicholinium-15, (53) 2-Methoxy-4-morpholinobenzoldiazoniumchlorid, Zinkchlorid, (54) Fomocain, (55) 4-Morpholinobenzophenon, (56) 4,4'-Ethylen-bis(2,6-morpholindion), (57) N,N'-Dicyclohexyl-4-morpholincarboxamidin, (58) Cyclohexyl-3-(2-morpholinoethyl)-2-thioharnstoff, (59) 4-Morpholinoacetophenon, (60) 4-(2-Chlorethyl)morpholin-Hydrochlorid, (61) 4-Morpholinethansulfonsäure, (62) 4-Morpholinpropansulfonsäure, (63) β-Hydroxymorpholinpropansufonsäure, (64) [N-(Aminoiminomethyl)-4-morpholincarboximidamid]-Hydrochlorid, (65) 4-Morpholincarbodithionsäureverbindung mit Morpholin, (66) 2,5-Dimethyl-4-(morpholinomethyl)phenol-Hydrochlorid-Monohydrat, (67) 1-Cyclohexyl-3-(2-morpholinoethyl)carbodiimidmetho-p-toluolsulfonat, (68) Hemicholinium-3[2,2'-(4,4'-biphenylen)bis(2-hydroxy-4,4-dimethylmorpholiniumbromid), (69) Hemicholinium-15[4,4-dimethyl-2-hydroxy-2-phenylmorpholiniumbromid], (70) 1-Aza-12-krone-4, (71) 1-Aza-15-krone-5, (72) 1-Aza-18-krone-6, (73) 1,4,10-Trioxa-7,13-diazacyclopentadecan, (74) 1,4,10,13-Tetraoxa-7,16-diazacyclooctadecan, (75) N,N'-Dibenzyl-1,4,10,13-tetraoxa-7,16-diazacyclioctadecan, (76) 4,7,13,18-Tetraoxa-1,10-diazabicyclo[8.5.5]eicosan, (77) 4,7,13,16,21-Pentaoxa-1,10-diazabicyclo[8.5.5]tricosan, (78) 4,7,13,16,21,24-Hexaoxa-1,10-diazabicyclo[8.8.8]hexacosan, (79) 5,6-Benzo-4,17,13,16,21,24-hexaoxa-1,10-diazabicyclo[8.8.8]hexacosan und (80) Mischungen davon; oder worin das transparentmachende Mittel eine Oxacyclische Verbindung ist; oder worin das transparentmachende Mittel ausgewählt ist aus der Gruppe bestehend aus: (A) Materialien der allgemeinen Formel: worin der gekrümmte Teil der Struktur eine Kohlenwasserstoffkette oder eine substituierte Kohlenwasserstoffkette bedeutet, worin zwei oder mehr Substituenten miteinander verbunden sein können, um einen Ring zu bilden; (B) Materialien der allgemeinen Formeln: worin R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ R₂₂, R₂₃, R₂₄, R₂₅, R₂₆, R₂₇ und R₂₈ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇ und R₂₈ miteinander verbunden sein können, um einen Ring zu bilden; (C) Materialien der allgemeinen Formel: worin der gekrümmte Teil der Struktur eine Kohlenwasserstoffkette oder eine substituierte Kohlenwasserstoffkette bedeutet, worin zwei oder mehr Substituenten miteinander verbunden sein können, um einen Ring zu bilden; (D) Materialien der allgemeinen Formeln: worin R₁, R₂, R₃, R₄, R₅, R₆, R₇ und R₈ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇ und R₈ miteinander verbunden sein können, um einen Ring zu bilden; (E) Materialien der allgemeinen Formeln: worin die gekrümmten Teile der Strukturen eine Kohlenwasserstoffkette oder eine substituierte Kohlenwasserstoffkette bedeuten, worin zwei oder mehr Substituenten miteinander verbunden sein können, um einen Ring zu bilden; (F) Materialien der allgemeinen Formel: worin R₁, R₂, R₃, R₄, R₅ und R₆ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅ und R₆ miteinander verbunden sein können, um einen Ring zu bilden; und (G) Mischungen davon; oder worin das transparentmachende Mittel ausgewählt ist aus der Gruppe bestehend aus (1) γ-Butyrolacton, (2) γ-Valerolacton, (3) γ-Caprolacton, (4) γ-Octanlacton, (5) γ-Nonanlacton, (6) γ-Decanolacton, (7) Undecan-γ-lacton, (8) γ-Phenyl-γ-butyrolacton, (9) α-Carbethoxy-γ-phenylbutyrolacton, (10) 2-Cumaranon, (11) β,β-Dimethyl-γ-(hydroxymethyl)-γ-butyrolacton, (12) γ-Ethoxycarbonyl-γ-butyrolacton, (13) 5-(Hydroxymethyl)-2(5H)-furanon, (14) Dihydro-4-4-dimethyl-2,3-furandion, (15) 2,5-Dimethyl-4-hydroxy-3(2H)-furanon, (16) Mevalon-(β-hydroxy-β-methyl-δ-valero)-lacton, (17) δ-Decanolacton, (18) Undecan-δ-lacton, (19) δ-Dodecanolacton, (20) Undecan-ω-lacton, (21) Oxacyclotridecan-2-on, (22) ω-Pentadecalacton, (23) Hydrindantin (2,2'-Dihydroxy-2,2'-biindan-1,1'3,3'-tetron, (24) Hydrindantin-Dihydrat, (25) 2-Oxepanon, (26) 4H-Pyran-2-on, (27) Methylcumalat, (28) Methyl-2-oxo-2H-pyran-3-carboxylat, (29) 4,6-Dimethyl-α-pyron, (30) 4-Methoxy-6-methyl-2H-pyran-2-on, (31) 3,6-Dihydro-4,6,6-trimethyl-2H-pyran-2-on, (32) 3,4-Dihydro-6-methyl-2H-pyran-2-on, (33) 3-Acetylcumarin, (34) 6-Methylcumarin, (35) 7-Ethoxycumarin, (36) Ethyl-3-cumarincarboxylat, (37) 7-Diethylamino-4-methylcumarin, (38) Dihydrocumarin, (39) 3-Brom-2-cumaranon, (40) Patulin, (41) 4H-Pyran-4-on, (42) 2-Ethyl-3-hydroxy-4H-pyran-4-on, (43) Butopyronoxyl(butyl-3,4-dihydro-2,2-dimethyl-4-oxo-2H-pyran-6-carboxylat, (44) Dehydroessigsäure, (45) 4-Chromon, (46) 4-Chromanon, (47) 4-Chromanol, (48) 6,7-Dimethoxy-2,2-dimethyl-4-chromanon, (49) 3-Isochromanon, (50) 6,7-Dimethoxy-3-isochromanon, (51) 6-Ethyl-4-oxo-4H-1-benzopyran-3-carbonitril, (52) 6-Ethyl-4-oxo-4H-1-benzopyran-3-carboxaldehyd, (53) 6-Isopropyl-4-oxo-4H-1-benzopyran-3-carbonitril, (54) 6-Isopropyl-4-oxo-4H-1-benzopyran-3-carboxaldehyd, (55) Maleinsäureanhydrid, (56) Brommaleinsäureanhydrid, (57) Citraconsäureanhydrid, (58) 2,3-Dimethylmaleinsäureanhydrid, (59) Dichlormaleinsäureanhydrid, (60) cis-Aconitsäureanhydrid, (61) Itaconsäureanhydrid, (62) Methylbemsteinsäureanhydrid, (63) Acetylmercaptobernsteinsäureanhydrid, (64) 2,2-Dimethylbemsteinsäureanhydrid (65) Phenylbemsteinsäureanhydrid, (66) 2-Octen-1-ylbemsteinsäureanhydrid, (67) 2-Dodecen-1-ylbernsteinsäureanhydrid, (68) 2-Octadecen-1-ylbernsteinsäureanhydrid, (69) 3-Oxabicyclo[3.1.0]hexan-2,4-dion, (70) Diglycolsäureanhydrid, (71) Glutarsäureanhydrid, (72) 3-Methylglutarsäureanhydrid, (73) 2,2-Dimethylglutarsäureanhydrid, (74) 3,3-Tetramethylenglutarsäureanhydrid, (75) 1-Cyclopenten-1,2-dicarbonsäureanhydrid, (76) 3,4,5,6-Tetrahydrophthalsäureanhydrid, (77) cis-1,2-Cyclohexandicarbonsäureanhydrid, (78) Hexahydro-4-methylphthalsäureanhydrid, (79) Methyl-5-norbomen-2,3-dicarbonsäureanhydrid, (80) 2,3-Pyridincarbonsäureanhydrid, (81) 3,4-Pyridincarbonsäureanhydrid, (82) Furfurylmercaptan, (83) S-Furfurylthioacetat, (84) Furfurylsulfid, (85) Furfurylmethyldisulfid, (86) Furfuryldisulfid, (87) Glycolaldehyddimer, (88) 6,7-Dihydrocyclopenta-1,3-dioxin-5(4H)-on, (89) (2R,6R)-tert-Butyl-6-methyl-1,3-dioxan-4-on, (90) 2,2-Dimethyl-1,3-dioxan-4,6-dion, (91) 3,6-Dimethyl-1,4-dioxan-2,5-dion, (92) 2,2,6-Trimethyl-4H-1,3-dioxin-4-on, (93) 2,2,5-Trimethyl-1,3-dioxan-4,6-dion, (94) 5-Brom-2,2,5-trimethyl-1,3-dioxan-4,6-dion, (95) 1,3-Dioxan-5,5-dimethanol, (96) 1,3,5-Trioxan, (97) 1,6-Dioxaspiro[4.4]nonan-2,7-dion, (98) 1,4-Dioxaspiro[4.5]decan-2-on, (99) 1,7-Dioxaspiro[5.5]undecan, (100) 2,4,8,10-Tetraoxaspiro[5.5]undecan, (101) 3,9-Divinyl-2,4,8-tetraoxaspiro[5.5]undecan, (102) 2,2-Pentamethylen-1,3-dioxalan, (103) 2-Phenyl-1,3-dioxalan, (104) 1,4-Cyclohexandionmonoethylenketal, (105) 1,4-Cyclohexandionbis(ethylenketal), (106) 1,4-Cyclohexandionmono-2,2-dimethyltrimethylenketal, (107) Piperonal, (108) Piperonylacetat, (109) Piperonylalkohol, (110) Piperonylnitril, (111) Piperonylamin, (112) 6-Nitropiperonal, (113) 6-Nitropiperonylalkohol, (114) 3',4'-(Methylendioxy)acetophenon, (115) 3,4-(Methylendioxy)anilin, (116) 2,3-(Methylendioxy)benzaldehyd, (117) 3,4-(Methylendioxy)phenylacetonitril, (118) 3,4-(Methylendioxy)toluol und (119) Mischungen davon; oder worin das transparentmachende Mittel ein Kronenether ist; oder worin das transparentmachende Mittel ausgewählt ist aus der Gruppe bestehend aus (1) 1,4,7,10-Tetraoxacyclododecan (12-Krone-4), (2) 2-(Hydroxyethyl)-12-krone-4, (3) 2-(Aminoethyl)-12-krone-4, (4) Benzo-12-krone-4, (5) 1,4,7,10,13-Pentaoxacyclododecan (15-Krone-5), (6) 2-(Hydroxyethyl)-15-krone-5, (7) 2-(Aminoethyl)-15-krone-5, (8) Benzo-15-krone-5, (9) 4'-Aminobenzo-15-krone-5, (10) 4'-Formylbenzo-15-krone-5, (11) 4'-Nitrobenzo-15-krone-5, (12) Bis[(benzo-15-krone-5)-15-ylmethyl]pimelat, (13) 1,4,7,10,13,16-Hexaoxacyclooctadecan (18-Krone-6), (14) 2-(Aminoethyl)-18-krone-6, (15) Benzo-18-krone-6, (16) 4'-Brombenzo-18-krone-6, (17) Dibenzo-18-krone-6, (18) Di-tert-butyldibenzo-18-krone-6, (19) cis-Dicyclohexan-18-krone-6, (20) Dibenzo-24-krone-8, (21) Dicyclohexano-24-krone-8, (22) Dibenzo-30-krone-10 und (23) Mischungen davon; oder worin das transparentmachende Mittel ein cyclischer Kohlenwasserstoff ist; oder worin das transparentmachende Mittel ausgewählt ist aus der Gruppe bestehend aus: (A) Materialien der allgemeinen Formeln: worin R₁, R₂, R₃, R₄, R₅, R₆, R₇, R₆, R₉, R₁₀, R₁₁ und R₁₂ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁ und R₁₂ miteinander verbunden sein können, um einen Ring zu bilden; (B) Materialien der allgemeinen Formel: worin R₁, R₂, R₃, R₄, R₅ und R₆ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅ und R₆ miteinander verbunden sein können, um einen Ring zu bilden; (C) Materialien der allgemeinen Formel: worin R₁, R₂, R₃, R₄, R₅, R₆, R₇, R₈, R₉ und R₁₀ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉ und R₁₀ miteinander verbunden sein können, um einen Ring zu bilden; (D) Materialien der allgemeinen Formeln: worin R₁, R₂, R₃, R₄, R₅, R₆, R₇, R₈, R₉, R₁₀, R₁₁ und R₁₂ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉, R₁₀, R₁₁ und R₁₂ miteinander verbunden sein können, um einen Ring zu bilden; (E) Materialien der allgemeinen Formel: worin R₁, R₂, R₃, R₄, R₅, R₆, R₇, R₈, R₉ und R₁₀ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆, R₇, R₈, R₉ und R₁₀ miteinander verbunden sein können, um einen Ring zu bilden; (F) Materialien der allgemeinen Formeln: worin R₁, R₂, R₃, R₄, R₅, R₆, R₇, R₈, R₉ und R₁₀ jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆ R₇, R₈, R₉ und R₁₀ miteinander verbunden sein können, um einen Ring zu bilden; (G) Materialien der allgemeinen Formel: worin der gekrümmte Teil der Struktur eine Kohlenwasserstoffkette oder eine substituierte Kohlenwasserstoffkette bedeutet, worin zwei oder mehr Substituenten miteinander verbunden sein können, um einen Ring zu bilden; und (H) Mischungen davon; oder worin das transparentmachende Mittel ausgewählt ist aus der Gruppe bestehend aus (1) Norbornan, (2) 2-Norbomancarbonitril, (3) 2-Norbomanmethanol, (4) 3-Methyl-2-norbornanmethanol, (5) Camphen, (6) Fenchylalkohol, (7) Thiocampher, (8) Norbornen, (9) 5-Norbomen-2-carbonitril, (10) 5-Norbornen-2-carboxaldehyd, (11) 5-Norbornen-2-methanol, (12) 5-Norbomen-2,2-dimethanol, (13) 5-Norbornen-2-benzoyl, (14) 2-Norbornanon, (15) 3-Chlor-2-norbomanon, (16) Fenchon, (17) 3-(Trifluoracetyl)campher, (18) 3-Heptafluorbutyrylcampher, (19) 3-Bromcampher, (20) 9,10-Dibromcampher, (21) 3,9,10-Tribromcampher, (22) Dicyclopentadien, (23) Methylcyclopentadiendimer, (24) Tricyclo[5.2.1]decan, (25) 4,8-Bis(hydroxymethyl)tricyclo[5.2.1.0^{2.6}]decan, (26) 8-Ketotricyclo[5.2.1.0^{2.6}]decan, (27) 3,4-Dimethoxy-3-cyclobuten-1,2-dion, (28) 3,4-Diethoxy-3-cyclobuten-1,2-dion, (29) 3,4-Diisopropoxy-3-cyclobuten-1,2-dion, (30) 3,4-Dibutoxy-3-cyclobuten-3-cyclobuten-1,2-dion, (31) 3-Methyl-2-(nitromethyl)-5-oxocyclopentanessigsäure, (32) 3-Ethyl-2-hydroxy-2-cyclopenten-1-on, (33) Methyl-4-methoxy-2-oxo-3-cyclopenten-1-carboxylat, (34) 3,3a,6,6a-Tetrahydro-2H-cyclopenta[b]furan-2-on, (35) 3a,4,5,6a-Hexahydro-5-hydroxy-4(hydroxymethyl)-2H-cyclopenta[b]furan-2-on, (36) 3-Methyl-1,2-cyclopentandion, (37) 4-Hydroxy-5-methyl-4-cyclopenten-1,3-dion-Monohydrat, (38) 2,4,4-Trimethylcyclohexen-1-on, (39) Ethyl-6-methyl-2-oxo-3-cyclohexen-1-carboxylat, (40) Ethyl-4-Hydroxy-6-methyl-2-oxo-3-cyclohexen-1 -carboxylat, (41) 5-(1-Acetoxy-1-methylethyl)-2-methyl-2-cyclohexen-1-on, (42) Thymochinon, (43) 2,6,6-Trimethyl-2-cyclohexen-1,4-dion, (44) Indan, (45) 1-Indanol, (46) 2-Indanol, (47) 1-Indanon, (48) 2-Indanon, (49) 2-Acetyl-1-tetralon, (50) 4-Methyl-1-tetralon, (51) 5,7-Dimethyl-1-tetralon, (52) 6,7-Dimethoxy-1-tetralon, (53) 1-Methyl-2-tetralon, (54) 6,7-Dimethoxy-2-tetralon, (55) Cyclohexanon, (56 Cycloheptanon, (57) Cyclooctanon, (58) Cyclononanon, (59) Cyclodecanon, (60) Cycloundecanon, (61) Cyclododecanon, (62) Cyclotridecanon, (63) Cyclopentadecanon, (64) 2-Acetylcyclohexanon, (65) 2-Allylcyclohexanon, (66) 2-Phenylcyclohexanon, (67) Cyclohexandion, (68) 2-Acetyl-1,3-cyclohexandion, (69) 4,4-Dimethyl-1,3-cyclohexandion, (70) 2-Acetyl-1,3-cyclopentandion, (71) 3,3,5,5-Tetramethyl-1,2-cyclopentandion, (72) Bicyclo[3.2.1]octan-2-on, (73) Endo-dimethyl-7-oxabicyclo[2.2.1]heptan-2,3-dicarboxylat, (74) Cineol, (75) Bicyclo[2.2.2]oct-5-en-2,3-dimethanol, (76) Tropon, (77) Tropolon, (78) Cyclooctenoxid, (79) 1,2,5,6-Diepoxycyclooctan, (80) 9-Methyl-Δ⁵⁽¹⁰⁾-octalin-1,6-dion, (81) cis-Bicyclo[3.3.0]octan-3.7-dion, (82) Azulen, (83) 1-Benzosuberon, (84) 1,5,9-Cyclododecatrien, (85) Cyclododecanepoxid, (86) 2,3-Cyclododecenopyridin, (87) 1,2,5,6,9,10-Hexabromcyclododecan, (88) 8-Cyclohexadecen-1-on, (89) Bicyclo[10.3.0]pentadec-12(1)-en-13-on, (90) 1,4,4a,8a-Tetrahydro-endo-1,4-methannaphthalin-5,8-dion, und (91) Mischungen davon; oder worin das transparentmachende Mittel ein Thioharnstoff ist; oder worin das transparentmachende Mittel ein Sulfon ist; oder worin das transparentmachende Mittel eine thiocyclische Verbindung ist; oder worin das transparentmachende Mittel ausgewählt ist aus der Gruppe bestehend aus Sulfiten, Sulfitderivaten, Sulfiden, Sulfidderivaten, quaternären Schwefelverbindungen, quaternären Schwefelderivaten und Mischungen davon; oder worin das transparentmachende Mittel eine Thiaaza-cyclische Verbindung ist; oder worin das transparentmachende Mittel ausgewählt ist aus der Gruppe bestehend aus (1) 1-Allyl-2-thiohamstoff, (2) 1-Methallyl-3-methyl-2-thioharnstoff, (3) 4-Allyl-3-thiosemicarbazid, (4) 1,3-Diethyl-2-thioharnstoff, (5) 1,3-Dibutyl-2-thioharnstoff, (6) 1-Benzyl-3-methyl-2-thiohamstoff, (7) 1,1,3,3-Tetramethyl-2-thiohamstoff, (8) 2-Imino-4-thiobiuret, (9) 1-Allyl-3-(2-hydroxyethyl)-2-thioharnstoff, (10) S-(2-Aminoethyl)isothiouroniumbromid-Hydrobromid, (11) S,S-Diphenylsulfillimin-Monohydrat, (12) Methylsulfon, (13) Ethylsulfon, (14) Butylsulfon, (15) Butadiensulfon, (16) Tetramethylensulfon, (17) 1,4-Butansulfon, (18) 1,4-Butandiol-cyclisches Sulfat, (19) Benzylsulfon, (20) Phenylsulfon, (21) Phenylvinylsulfon, (22) Phenylstyrolsulfon, (23) Phenyl-2-(trimethylsilyl)methylsulfon, (24) Phenyl-2-(trimethylsilyl)ethylsulfon, (25) Phenyl-2-(trimethylsilyl)ethinylsulfon, (26) 4-(Fluorphenyl)sulfon, (27) 4-(Fluorphenyl)methylsulfon, (28) Chlormethylphenylsulfon, (29) Chlormethyl-p-tolylsulfon, (30) 2-Chlorethylphenylsulfon, (31) Methylthiomethylphenylsulfon, (32) Methylthiomethyl-p-tolylsulfon, (33) 2-(Phenylsulfonyl)tetrahydropyran, (34) 1-(Phenylsulfonyl)indol, (35) 1-(p-Toluolsulfonyl)imidazol, (36) 1-(p-Tosyl)-3,4,4-trimethylimidazolidin, (37) 4-(p-Tosylsulfonyl)hexahydro-1,4-thiazepin, (38) Thionaphthen, (39) 4-Keto-4,5,6,7-tetrahydrothianaphthen, (40) 2,2'-Bithiophen, (41) 2,2':5',2"-Terthiophen, (42) N-Acetylhomocystein-Thiolacton, (43) Tetrahydrothiopyran-4-on, (44) Thiochroman-4-on, (45) Thiochroman-4-ol, (46) Thioctansäure, (47) Ethyl-1,3-dithiolan-2-carboxylat, (48) 3H-1,2-Benzodithiol-3-on, (49) 1,3-Dithian, (50) 2-Phenyl-1,3-dithian, (51) Ethyl-1,3-dithian-2-carboxylat, (52) 5,6-Dihydro-5-methyl-4H-1,3,5-dithiazin, (53) 1,4-Dithian, (54) 2,5-Dihydroxy-2,5-dimethyl-1,4-dithian, (55) 1,5-Dithiacyclooctan-3-ol, (56) 1,4-Dithiaspiro[45]decan-8-ol, (57) 1,3,5-Tithian, (58) 1,4,7-Trithiacyclononan, (59) 1,4,7-Trithiacyclodecan, (60) 1,4,7,10-Tetrathiacyclododecan, (61) 3,6,9,14-Tetrathiabicyclo[9.2.1]tetradeca-11,13-dien, (62) 1,4,8,1-Tetrathiacyclotetradecan, (63) 1,5,9,13-Tetrathiocyclohexadecan, (64)1,5,9,13-Tetrathiacyclohexadecan-3,11-diol, (65)1,4,7,10,13-Pentathiacyclopentadecan, (66)1,4,7,10,13,16-Hexathiacyclooctadecan, (67) 1,5,9,13,17,21-Hexathiacyclotetracosan-3,11,19-triol, (68)1,4,7,10,13,16,19,22-Octathiacyclotetracosan, (69) 1,4,8,11,15,18,22,25-Octathiacyclooctacosan, (70) 1,4,7,10,13,16,19,22,25-Nonathiacycloheptacosan, (71) Dimethylsulfit, (72) Diethylsulfit, (73) Natriumsulfit, (74) Allyldisulfid, (75) Aminophenyldisulfid, (76) Benzyldisulfid, (77) Benzylphenylsulfid, (78) Trimethylsulfoniummethylsulfat, (79) (2-Chlorethyl)dimethylsulfoniumiodid, (80) 3-(Chlorpropyl)diphenylsulfoniumtetrafluorborat, (81) Trimethylsulfoniumiodid, (82) Trimethylsulfoxoniumiodid, (83) Trimethylsulfoxoniumchlorid, (84) Triphenylmethansulfenylchlorid, (85) Dimethyl(2-methoxy-5-nitrobenzyl)sulfoniumbromid, (86) Thioninperchlorat, (87) p-Xylylenbis(tetrahydrothiopheneumchlorid), (88) Tris(dimethylamino)sulfoniumdifluortrimethylsilicat, (89) Tris(dimethylamino)sulfoniumtrifluormethoxid, (90) (3-Amino-3-carboxypropyl)dimethylsulfoniumchlorid und (91) Mischungen davon; oder worin das transparentmachende Mittel eines der folgenden allgemeinen Formeln ist: worin R₁, R₂, R₃, R₄, R₅, R₆ und R₇, jeweils unabhängig voneinander ausgewählt sind aus der Gruppe bestehend aus Wasserstoffatomen, Alkylgruppen, substituierten Alkylgruppen, Arylgruppen, substituierten Arylgruppen, Arylalkylgruppen, substituierten Arylalkylgruppen, Hydroxygruppen, Amingruppen, Imingruppen, Ammoniumgruppen, Pyridingruppen, Pyridiniumgruppen, Ethergruppen, Aldehydgruppen, Ketongruppen, Estergruppen, Amidgruppen, Carbonsäuregruppen, Carbonylgruppen, Thiocarbonylgruppen, Sulfatgruppen, Sulfonatgruppen, Sulfidgruppen, Sulfoxidgruppen, Phosphingruppen, Phosphoniumgruppen, Phosphatgruppen, Cyangruppen, Nitrilgruppen, Mercaptogruppen, Nitrosogruppen, Halogenatomen, Nitrogruppen, Sulfongruppen, Acylgruppen, Säureanhydridgruppen und Azidgruppen, worin zwei oder mehr von R₁, R₂, R₃, R₄, R₅, R₆ und R₇ miteinander verbunden sein können, um einen Ring zu bilden; oder worin das transparentmachende Mittel ausgewählt ist aus der Gruppe bestehend aus (1) 2-Amino-2-thiazolin, (2) 2-Aminothiazol, (3) 2-Amino-4-methylthiazol, (4) 2-Amino-4-methylthiazol, (5) 2-Amino-4-thiazolessigsäure, (6) 2-Acetamido-4-methylthiazol, (7) 2-Acetylthiazol, (8) 5-Acetyl-2,4-dimethylthiazol, (9) 4-Methyl-5-vinylthiazol, (10) 2-Amino-4-phenyl-5-tetradecylthiazol, (11) 2,4-Thiazolidindion, (12) 3-Aminorhodanin, (13) 3-Methylrhodanin, (14) 3-Ethylrhodanin, (15) 3-Allylrhodanin, (16) 3-Hydroxy-4-methyl-2(3H)-thiazolethion, (17) Benzothiazol, (18) 2-Methylbenzothiazol, (19) 2-(Methylthio)benzothiazol, (20) 2-Amino-4-methylbenzothiazol, (21) 3-Methylbenzothiazol-2-thion, (22) 2,1,3-Benzothiadiazol, (23) 4-Amino-2,1,3-benzothiadiazol, (24) 3,4-Dimethyl-5-(2-hydroxyethyl)thiazoliumiodid, (25) 3-Ethyl-5-(2-hydroxyethyl)4-methylthiazoliumbromid, (26) 2-Amino-5-nitrothiazol, (27) 2-Amino-a-(methoxyimino)-4-thiazolessigsäure, (28) Ethyl-2-amino-α-(hydroxyimino)-4-thiazolacetat, (29) Ethyl-2-amino-a-(methoxyimino)-4-thiazolacetat, (30) Ethyl-2-amino-4-thiazolacetat, (31) Ethyl-2-amino-4-thiazolglyoxylat, (32) 1-Phenyl-3-(2-thiazolyl)-2-thioharnstoff, (33) 2-Amino-4-methoxybenzothiazol, (34) 2-Amino-5,6-dimethylbenzothiazol, (35) N'-(2-Thiazolyl)sulfanilamid, (36) 6-Ethoxy-2-benzothiazolsulfonamid, (37) Ethyl-2-(formylamino)-4-thiazolacetat, (38) Ethyl-2-(formylamino)-4-thiazolglyoxylat, (39) 2-(Formylamino)-a-(methoxyimino)-4-thiazolessigsäure, (40) 2-Acetamido-4-methyl-5-thiazolsulfonylchlorid, (41) 2-Thioxo-4-thiazolidincarbonsäure, (42) Thiazolidin-4-carbonsäure, (43) Pseudothiohydantoin, (44) 2-Amino-1,3,4-thiadiazol, (45) 2-Amino-5-trifluormethyl-1,3,4-thiadiazol, (46) 2-Amino-5-methyl-1,3,4-thiadiazol, (47) 2-Amino-5-ethyl-1,3,4-thiadiazol, (48) 2-Amino-5-(ethylthio)-1,3,4-thiadiazol, (49) 5-Amino-1,3,4-thiadiazol-2-thiol, (50) 2-Acetamido-5-benzylthio-1,3,4-thiadiazol, (51) 5-Acetamido-1,3,4-thiadiazol-2-sulfonamid, (52) 5-Anilino-1,2,3,4-thiatriazol, (53) 2-Amino-4,5-dimethylthiazol-Hydrochlorid, (54) 2-Amino-4-imino-2-thiazolin-Hydrochlorid, (55) 2-Amino-2-thiazolin-Hydrochlorid, (56) 2-Amino-5-bromthiazol-Monohydrobromid, (57) 5-Amino-3-methylisothiazol-Hydrochlorid, (58) 3-Methyl-2-benzothiazolinonhydrazon-Hydrochlorid-Hydrat, (59) 5-Amino-2-methylbenzothiazol-Dihydrochlorid, (60) 2,4-Diamino-5-phenylthiazol-Monohydrobromid, (61) 2-Amino-4-phenylthiazol-Hydrobromid-Monohydrat, (62) 2-(Tritylamino)-α-(methoxyimino)-4-thiazolessigsäure-Hydrochlorid, (63) (2,3,5,6-Tetrahydro-6-phenylimidazo[2,1-b]thiazol-Hydrochlorid, (64) 3-Ethyl-2-methyl-2-thiazoliumiodid, (65) 3-Benzyl-5-(2-hydroxyethyl)-4-methylthiazoliumchlorid, (66) Thiamin-Hydrochlorid, (67) 3-(Carboxymethyl)benzothiazoliumbromid, (68) 2-Azido-3-ethylbenzothiazoliumtetrafluorborat, (69) 3-Ethyl-2-methylbenzothiazoliumiodid, (70) 2-Methyl-3-propylbenzothiazoliumiodid, (71) 3-Ethyl-2-(2-hydroxy-1-propenyl)benzothiazoliumchlorid, (72) 3,6-Dimethyl-2-(4-dimethylaminophenyl)benzothiazoliumbromid, (73) Trifluorperazin-Dihydrochlorid, (74) Thioridazin-Hydrochlorid, (75) Promethazin-Hydrochlorid, (76) Ethopropazin-Hydrochlorid, (77) Chlorpromazin-Hydrochlorid und (78) Mischungen davon; oder worin das transparentmachende Mittel ausgewählt ist aus der Gruppe bestehend aus Phosphinen, Phosphiten, cyclischen Phosphorverbindungen, Phosphinoxiden, quatemären Phosphoniumsalzen und Mischungen davon; oder worin das transparentmachende Mittel ausgewählt ist aus der Gruppe bestehend aus (1) Triphenylphosphin, (2) Tri-m-tolylphosphin, (3) Tris(3-methoxyphenyl)phosphin, (4) Tris(4-chlorphenyl)phosphin, (5) Tris(pentafluorphenyl)phosphin, (6) Tricyclohexylphosphin, (7) Tribenzylphosphin, (8) Tri-2-furylphosphin, (9) Bis(pyrrolidino)methoxyphosphon, (10) Tetraphenylbiphosphin, (11) 1,3-Bis(diphenylphosphino)propan, (12) 1,5-Bis(diphenylphosphino)pentan, (13) 1,6-Bis(diphenylphosphino)hexan, (14) lsopropyldiphenylphosphin, (15) Diphenyl(p-tolyl)phosphin, (16) (4-Bromphenyl)diphenylphosphin, (17) Diphenyl-2-pyridylphosphin, (18) Dicyclohexylphenylphosphin, (19) Trimethylphosphit, (20) Triethylphosphit, (21) Tris(2-chlorethyl)phosphit, (22) Tributylphosphit, (23) Triphenylphosphit, (24) Trimethylphosphit-Kupferiodid, (25) Triethylphosphit-Kupferiodid, (26) Dipropylphosphit, (27) Bis(2-ethylhexyl)phosphit, (28) Bis(4-Nitrobenzyl)phosphit, (29) 2,2'-Ethylidenbis(4,6-di-tert-butylphenyl)fluorphosphit, (30) Pentaerythritdiphenyldiphosphit, (31) 2-Furyltetramethylphosphorodiamidat, (32) Diethyl(pyrrolidinomethyl)phosphonat, (33) Cyclophosphamid-Monohydrat, (34) 2-Chlor-1,3,2-dioxaphospholan-2-oxid, (35) N,N-Diethyl-1,5-dihydro-2,4,3-benzodioxaphosphepin-3-amin, (36) 1,2-Phenylenphosphochloridit, (37) 1,2-Phenylenphosphochloridat, (38) 2-Chlor-4H-1,3,2-benzodioxaphosphorin-4-on, (39) 2,4-Bis(methylthio)-1,3-dithia-2,4-diphosphetan-2,4-disulfid, (40) Triphenylphosphinoxid, (41) Tris(hydroxymethyl)phosphinoxid, (42) Trimethoxyphosphinoxid, (43) Triethoxyphosphinoxid, (44) Triphenoxyphosphinoxid, (45) Tris(2-butoxyethoxy)phosphinoxid, (46) Diphenylphosphinoxid, (47) Diphenyl(2,4,6-trimethylbenzoyl)phosphinoxid, (48) Phenylphosphinsäure, (49) Diphenylphosphat, (50) Vinylphosphonsäure, (51) Propylphosphonsäure, (52) Pyrophosphorsäure, (53) Triphenylphosphat, (54) Tetrabutylphosphoniumchlorid, (55) Tetrabutylphosphoniumbromid, (56) Hexadecyltributylphosphoniumbromid, (57) Stearyltributylphosphoniumbromid, (58) Azidotris(diethylamino)phosphoniumbromid, (59) Phosphonitrilchloridtrimer, (60) Tetramethylphosphoniumbromid, (61) Tetramethylphosphoniumchlorid, (62) Tetraethylphosphoniumbromid, (63) Tetraethylphosphoniumchlorid, (64) Tetraethylphosphoniumiodid, (65) Tetraphenylphosphoniumbromid, (66) Tetraphenylphosphoniumchlorid, (67) Tetraphenylphosphoniumiodid, (68) Methyltriphenylphosphoniumbromid, (69) Methyltriphenylphosphoniumiodid, (70) Ethyltriphenylphosphoniumbromid, (71) n-Propyltriphenylphosphoniumbromid, (72) lsopropyltriphenylphosphoniumiodid, (73) Cyclopropyltriphenylphosphoniumbromid, (74) n-Butyltriphenylphosphoniumbromid, (75) Isobutyltriphenylphosphoniumbromid, (76) Hexyltriphenylphosphoniumbromid, (77) Benzyltriphenylphosphoniumchlorid, (78) Brommethyltriphenylphosphoniumbromid, (79) Chlormethyltriphenylphosphoniumchlorid, (80) 3-Brompropyltriphenylphosphoniumbromid, (81) 3-Brombutyltriphenylphosphoniumbromid, (82) 4-Brombutyltriphenylphosphoniumbromid, (83) 2-Dimethylaminoethyltriphenylphosphoniumbromid, (84) [(3-Dimethylamino)propyl]triphenylphosphoniumbromid, (85) 2-Hydroxyethyltriphenylphosphoniumbromid, (86) (2-Hydroxyethyl)triphenylphosphoniumchlorid, (87) [3-Hydroxy-2-methylpropyl]triphenylphosphoniumbromid, (88) [3-Hydroxy-2-methylpropyl]triphenylphosphoniumbromid, (89) (2-Hydroxybenzyltriphenylphosphoniumbromid, (90) (Formylmethyl)triphenylphosphoniumchlorid, (91) (Methoxymethyl)triphenylphosphoniumchlorid, (92) Acetonyltriphenylphosphoniumchlorid, (93) Carbomethoxymethyltriphenylphosphoniumbromid, (94) (Ethoxycarbonylmethyl)triphenylphosphoniumchlorid, (95) Carbethoxymethyltriphenylphosphoniumbromid, (96) (tert-Butoxycarbonylmethyl)triphenylphosphoniumbromid, (97) Phenacyltriphenylphosphoniumbromid, (98) (4-Ethoxybenzyl)triphenylphosphoniumbromid, (99) 4-Butoxybenzyltriphenylphosphoniumbromid, (100) 2-(1,3-Dioxan-2-yl)ethyl]triphenylphosphoniumbromid, (101) (1,3-Dioxolan,2-ylmethyl)triphenylphosphoniumbromid, (102) Vinyltriphenylphosphoniumbromid, (103) Allyltriphenylphosphoniumbromid, (104) Allyltriphenylphosphoniumchlorid, (105) Propargyltriphenylphosphoniumbromid, (106) (3-Trimethylsilyl-2-propinyl)triphenylphosphoniumbromid, (107) p-Xylylenbis(triphenylphosphoniumbromid) und (108) Mischungen davon; oder worin das transparentmachende Mittel ein Nitril ist; oder worin das transparentmachende Mittel ausgewählt ist aus der Gruppe bestehend aus (1) Cyanacetohydrazid, (2) 4,4-Dimethyl-3-oxopentannitril, (3) 1-Cyan-N-methylthioformamid, (4) Cyanmethyl-N,N-dimethyldithiocarbamat, (5) 4-Hydroxy-3-methoxy-phenylacetonitril, (6) Tosylcyanid, (7) Tosylmethylisocyanid, (8) 5-Fluor-2-methylbenzonitril, (9) 2-Fluor-5-methylbenzonitril, (10) 4-(Methylthio)benzonitril, (11) 4-(Dimethylamino)benzonitril, (12) 3,4-Dimethoxybenzonitril, (13) 4-Hydroxy-3-methoxybenzonitril, (14) 4-(trans-4-Pentylcyclohexyl)benzonitril, (15) 4'-Pentyl-4'-biphenylcarbonitril, (16) 4'-(Pentyloxy)-4-biphenylcarbonitril, (17) 4'-Hexyl-4-biphenylcarbonitril, (18) 4'-(Hexyloxy)-4-biphenylcarbonitril, (19) 4'-Heptyl-4-biphenylcarbonitril, (20) 4'-Heptyloxy-4-biphenylcarbonitril, (21) 4'-Octyl-4-biphenylcarbonitril, (22) 4'-(Octyloxy)-4-biphenylcarbonitril, (23) Succinonitril, (24) Fumaronitril, (25) 1,4-Dicyan-2-buten, (26) (Dimethylaminomethylen)malononitril, (27) (1-Ethoxyethyliden)malononitril, (28) a-Chlorbenzylidenmalononitril, (29) Benzylidenmalononitril, (30) 2-Benzoyloxy-2-phenylmalononitril, (31) O-(p-Tosyl)isonitrosomalononitril, (32) Tetrafluorphthalonitril, (33) Iminodiacetonitril, (34) Phenylendiacetonitril, (35) 3,3'-(4-Formylphenylimino)dipropionitril, (36) Tris(2-cyanethyl)nitromethan, (37) 1,1,3,3-Propantetracarbonitril, (38) Tetracyanethylenoxid und (39) Mischungen davon; oder worin das transparentmachende Mittel ausgewählt ist aus der Gruppe bestehend aus Isothiocyanaten, Isocyanaten und Mischungen davon; oder worin das transparentmachende Mittel ausgewählt ist aus der Gruppe bestehend aus (1) 4-Azidophenylisothiocyanat, (2) 1-Naphthylisothiocyanat, (3) 4-Dimethylamino-1-naphthylisothiocyanat, (4) 1-lsothiocyanato-4-(trans-4-propylcyclohexyl)benzol, (5) 1-(trans-4-Hexylcyclohexyl)-4-isothiocyanatobenzol, (6) 1-(4-trans-Hexylcyclohexyl)-4-[2-(4-isothiocyanatophenyl)]benzol, (7) 1-lsothiocyanato-4-(trans-4-octylcyclohexyl)benzol, (8) 4-lsothiocyanatophenyl-4-pentabicyclo[2.2.2]octan-1-carboxylat, (9) Benzylthiocyanat, (10) Guanidinthiocyanat, (11) Methylendithiocyanat, (12) 4,4'-Methylenbis(phenylisocyanat), (13) 4,4'-Methylenbis(2,6-diethylisocyanat) und (14) Mischungen davon; oder worin das transparentmachende Mittel ausgewählt ist aus der Gruppe bestehend aus Oximverbindung, Hydroxamsäureverbindungen und Mischungen davon; oder worin das transparentmachende Mittel ausgewählt ist aus der Gruppe bestehend aus (1) Formamidoxim, (2) Acetaldoxim, (3) Pyruvinaldehyd-1-oxim, (4) Acetonoxim, (5) Ethylchloroximidoacetat, (6) 2,3-Butandionmonoxim, (7) 5-Hydroxypentenaloxim, (8) Cyclopentanonoxim, (9) Cyclohexanonoxim, (10) Cyclooctanonoxim, (11) Benzaldehydoxim, (12) 2-Nitrobenzaldehydoxim, (13) Salicylaldoxim, (14) 2-lsonitrosoacetphenon, (15) 1-Phenyl-1,2-Propandion-2-oxim, (16) 2-Pyridinaldoxim, (17) Nifuroxim und (18) Mischungen davon; oder worin das transparentmachende Mittel ein Hydroxamsäurederivat ist; oder worin das transparentmachende Mittel ausgewählt ist aus der Gruppe bestehend aus (1) Acetohydroxamsäure, (2) Suberohydroxamsäure, (3) Mandelohydroxamsäure, (4) Benzohydroxamsäure, (5) N-Phenylbenzohydroxamsäure und (6) Mischungen davon; oder worin das transparentmachende Mittel ausgewählt ist aus der Gruppe bestehend aus Alkylammoniumsalzen, Arylammoniumsalzen, Arylalkylammoniumsalzen oder Mischungen davon; oder worin das transparentmachende Mittel ausgewählt ist aus der Gruppe bestehend aus (1) Tetramethylammoniumfluorid-Tetrahydrat, (2) Tetraethylammoniumacetat-Tetrahydrat, (3) Tetrabutylammoniumchlorid, (4) Tetrabutylammoniumchlorid-Hydrat, (5) Tetrabutylammoniumbromid, (6) Tetrabutylammoniumtribromid, (7) Tetrabutylammoniumacetat, (8) Tetrabutylammoniumthiocyanat, (9) Tetrapentylammoniumbromid, (10) Tetrahexylammoniumbromid, (11) Tetrahexylammoniumchlorid, (12) Tetrahexylammoniumhydrogensulfat, (13) Tetraheptylammoniumchlorid, (14) Tetraheptylammoniumbromid, (15) Tetraoctylammoniumbromid, (16) Tetrakisdecylammoniumbromid, (17) Tetrahexadecylammoniumbromid, (18) Tetramethylammoniumbromid, (19) Tetramethylammoniumchlorid, (20) Tetramethylammoniumiodid, (21) Tetraethylammoniumbromid, (22) Tetraethylammoniumchlorid, (23) Tetraethylammoniumiodid, (24) Tetrapropylammoniumbromid, (25) Tetrapropylammoniumiodid, (26) Tetrabutylammoniumiodid, (27) Tetrapentylammoniumchlorid, (28) Tetrahexylammoniumbromid, (29) Tetrahexylammoniumiodid, (30) Tetradecylammoniumbromid, (31) Tetradodecylammoniumbromid, (32) Tetraoctadecylammoniumbromid, (33) Methyltrioctylammoniumbromid, (34) Tridodecylmethylammoniumchlorid, (35) Tridodecylammoniumiodid, (36) N-Dodecyl-N-methylephedriniumbromid, (37) Phenyltrimethylammoniumtribromid, (38) Tricaprylmethylammoniumchlorid, (39) Tridodecylmethylammoniumchlorid, (40) Tridecyloxypropyldihydroxyethylmethylammoniumchlorid, (41) N-Tetradecyldimethylnaphthylmethylammoniumchlorid, (42) Octadecyldiethanolmethylammoniumchlorid, (43) Octadecyldihydroxyethylmethylammoniumchlorid, (44) dihydriertes Talgbenzylmethylammoniumchlorid, (45) 2-Aminoethyltrimethylammoniumchlorid-Hydrochlorid, (46) 2-Bromethyltrimethylammoniumbromid, (47) 2-Chlorethyltrimethylammoniumchlorid (48) 3-Carboxypropyltrimethylammoniumchlorid, (49) [3-(Methacryloylamino)propyl]trimethylammoniumchlorid, (50) Phenyltrimethylammoniumbromid, (51) Phenyltrimethylammoniumchlorid, (52) Phenyltrimethylammoniumiodid, (53) Benzyltrimethylammoniumchlorid, (54) Benzyltrimethylammoniumbromid, (55) 4-Nitrobenzyltrimethylammoniumchlorid, (56) [2-(4-Nitrophenyl)allyl]trimethylammoniumiodid, (57) Kokostrimethylammoniumchlorid, (58) Palmityltrimethylammoniumchlorid, (59) Myristyltrimethylammoniumbromid, (60) Oleyltrimethylammoniumchlorid, (61) Soyatrimethylammoniumchlorid, (62) Talgtrimethylammoniumchlorid, (63) hydriertes Talgtrimethylammoniumchlorid, (64) Stearyltrimethylammoniumchlorid, (65) Behenyltrimethylammoniumchlorid, (66) Guarhydroxypropyltrimethylammoniumchlorid, (67) Benzyltriethylammoniumbromid, (68) Butyltripropylammoniumbromid, (69) Methyltributylammoniumchlorid, (70) Methyltributylammoniumbromid, (71) Methyltributylammoniumiodid, (72) Benzyltributylammoniumchlorid, (73) Benzyltributylammoniumbromid, (74) Benzyltributylammoniumiodid, (75) Heptyltributylammoniumbromid, (76) Benzyldodecyldimethylammoniumbromid, (77) Benzyltetradecyldimethylammoniumchlorid-Dihydrat, (78) Benzylcetyldimethylammoniumchlorid-Monohydrat, (79) Benzylstearyldimethylammoniumchlorid-Monohydrat, (80) N,N-Dimethylmethylenammoniumchlorid, (81) N,N-Dimethylmethylenammoniumiodid, (82) Chlormethylendimethylammoniumchlorid, (83) Dichlormethylendimethylammoniumchlorid, (84) Dimethylaminomethylenaminomethylendimethylammoniumchlorid, (85) Benzethoniumchlorid, (86) Methylbenzethoniumchlorid, (87) 1-Propanaminium-2,3-dihydroxy-N-dimethyl-N-[3(oxococoyl)amino]propyl]-chlorid, (88) Cetyldimethylethylammoniumbromid, (89) Octyldodecyldimethylammoniumchlorid, (90) Dodecyl(2-hydroxy-1-methyl-2-phenyl-ethyl)dimethylammoniumbromid, (91) Dodecyldimethyl-2-phenoxyethylammoniumbromid, (92) Dodecanoyl-N-methylaminoethyl(phenylcarbamylmethyl)dimethylammoniumchlorid, (93) 3-Chlor-2-hydroxypropyl-N,N,N-dimethyldodecylammoniumchlorid, (94) 3-Chlor-2-hydroxypropyl-N,N,N-dimethyloctadecylammoniumchlorid, (95) Dodecylbenzyldimethylammoniumbromid, (96) Dodecylbenzyldimethylammoniumchlorid, (97) Kokosbenzyldimethylammoniumchlorid, (98) Benzyltetradecyldimethylammoniumchlorid, (99) Benzylcetyldimethylammoniumchlorid, (100) Benzyloctadecyldimethylammoniumchlorid, (101) Benzyltalgdimethylammoniumchlorid, (102) Benzyl-hydriertes-talgdimethylammoniumchlorid, (103) Benzylbehenyldimethylammoniumchlorid, (104) Dioctyldimethylammoniumchlorid, (105) Didecyldimethylammoniumchlorid, (106) Didecyldimethylammoniumbromid, (107) Dikokosdimethylammoniumchlorid, (108) Dicetyldimethylammoniumchlorid, (109) Disoyadimethylammoniumchlorid, (110) Ditalgdimethylammoniumchlorid, (111) dihydriertes Talgdimethylammoniumchlorid, (112) Dibehenyl/Diarachidyldimethylammoniumchlorid, (113) Soyaamidopropylbenzyldimethylammoniumchlorid, (114) Soyadikokos-quatemäres-ammoniumchlorid, (115) Gluconamidopropyldimethyl-2-hydroxyethylammoniumchlorid, (116) N-Alkyl-N-N-dimethyl-N(dodecylacetat)ammoniumchlorid, worin Alkyl 14 bis 20 Kohlenstoffatome hat, (117) Nerzamidopropyldimethyl-2-hydroxyethylammoniumchlorid, (118) N-Raps-(3-amidopropyl)-N-N-dimethyl-N-(2,3-epoxypropyl)ammoniumchlorid, (119) N-Stearyl-(3-amidopropyl)-N-benzyldimethylammoniumchlorid, (120) Rapsamidopropylbenzyldimethylammoniumchlorid, (121) Rapsamidopropylethyldimethylammoniumchlorid, (122) Kokamidopropylpolyethylenglycoldimethylammoniumchloridphosphat, (123) Butyrylcholinchlorid und (124) Mischungen davon; oder worin das transparentmachende Mittel ausgewählt ist aus der Gruppe bestehend aus Piperidinthiocyanat, 2-Piperidinmethanol, Bis(pentamethylenharnstoff, 4,4'-Trimethylen-bis(1-piperidinpropionitril), Tripiperidinphosphinoxid, Homopiperazin, 1-Piperonylpiperazin, Hexacyclentrisulfat, 5,10,15,20-Tetraphenyl-21H,23H-porphin, 5,10,15,20-Tetrakis(4-methoxyphenyl)-2H,23H-porphin, Pyrrol-2-carboxaldehyd, 3-Pyrrolidino-1,2-propandiol, Pyrazol, 3-Aminopyrazol, Imidazol, 2-Ethylimidazol, 2-(2-Piperidinoethyl)pyridin, 1-Dodecylpyridiniumchlorid, Pyridiniumbromidperbromid, 3-Aminochinolin, 8-Hydroxychinolin, 7,8-Benzochinolin, 8-Hydroxychinaldin, Chinoxalin, 4,5-Dihydro-6-methyl-3(2H)-pyridazinon-Monohydrat, Phthalazin, 1,10-Phenanthrolin, 1,3,5-Triazin, Trichlormelamin, Trichlorisocyanursäure, Norboman, Tricyclo[5.2.1.0]decan, Norcampher, Tropolon, 1-Indanol, trans,trans,cis-1,5,9-Cyclododecatrien, Cyclodecanepoxid, 2,3-Cyclododecanpyridin, 1,2,5,6,9,10-Hexabromcyclododecan, 1,4,4a,8a-Tetrahydro-endo-1,4-methano-naphthalin-5,8-dion, γ-Butyrolacton, β,β-Dimethyl-γ-(hydroxymethyl)-γ-butyrolacton, 2,5-Dimethyl-4-hydroxy-3(2H)-furanon, Hydrindantin-Dihydrat, 2,4,8,10-Tetraoxaspiro[5.5]undecan, 1,3,5-Trioxan, Cyclooctanon, Piperonal, Piperonylalkohol, Piperonylnitril, 3,4(Methylendioxy)phenylacetonitril, Maleinsäureanhydrid, S-Acetylmercaptobemsteinsäureanhydrid, 2-Octadecen-1-ylbernsteinsäureanhydrid, 18-Krone-6, Benzo-18-krone-6, Dibenzo-18-krone-6, Dibenzo-24-krone-8, 5-Amino-3-methylisooxazol, 2-Oxazolidon, 5,5-Dimethyloxazolidin-2,4-dion, 3-Ethyl-2-thioxo-4-oxazolidinon, 3-Morpholino-1,2-propandiol, 4-Phenylmorpholin, N, N'-Dibenzyl-1,4,10,13-tetraoxa-7,16-diazacyclooctadecan, 4,7,13,16,21,24-Hexaoxa-1,10-diazabicyclo[8.8.8]hexacosan, γ-Valerolactam, ε-Caprolactam, 2-Azacyclooctanon, 2-Azacyclononanon, Maleimid, N-Methylsuccinimid, Phthalimid-DBU-Salz, 1-Allyl-2-thioharnstoff, 1,3-Dithian, 1-Benzyl-3-methyl-2-thioharnstoff, 2-lmino-4-thiobiuret, Butylsulfon, 2,2'-Bithiophen, 2-Phenyl-1,3-dithian, 3,6,9,14-Tetrathiabicyclo[9.2.1]tetradeca-11,13-dien, 1,5,9,13-Tetrathiacyclohexadecan-3,11-diol, 1,4,7,10,13-Penta-thiacyclopentadecan, 2-Aminothiazol, 2-Amino-2-thiazolin, 3-Methylrhodanin, 3-Ethyl-5-(2-hydroxyethyl)-4-methylthiazoliumbromid, Triphenylphosphin, Tricyclohexylphosphin, 1,3-Bis(diphenylphosphino)propan, 1,5-Bis(diphenylphosphino)pentan, Isopropyldiphenylphosphin, Triethylphosphit, Triphenylphosphit, Triethylphosphit-Kupferiodid, Dipropylphosphit, Bis(2-ethylhexyl)phosphit, Bis(4-nitrobenzyl)phosphit, Diphenylphosphinoxid, Diphenyl(2,4,6-trimethylbenzoyl)phosphinoxid, Vinylphosphonsäure, Cyanacetohydrazid, Cyanmethyl-N,N-dimethyldithiocarbamat, 4'-Pentyl-4'-biphenylcarbonitril, 4'-(Octyloxy)-4-biphenylcarbonitril, 1,4-Dicyan-2-buten, Benzylidenmalononitril, 1-lsothiocyanato-4-(trans-4-propylcyclohexyl)benzol, Formamidoxim, Ethylchloroximidoacetat, Acetohydroxamsäure, Tetrahexylammoniumchlorid, Tetraheptylammoniumchlorid, Tetraheptylammoniumbromid und Mischungen davon.

9. Ein Verfahren welches umfaßt (1) das Migrationsbilderzeugungselementes gemäß Anspruch 1 umfassend (a) ein Substrat, (b) eine erweichbare Schicht umfassend ein erweichbares Material und ein photoempfindliches Migrationsmarkierungsmaterial und (c) ein transparentmachendes Mittel, welches das damit in Kontakt befindliche Migrationsmarkierungsmaterial transparent macht, enthalten in mindestens einer Schicht des Migrationsbilderzeugungselementes; (2) gleichmäßiges Laden des Bilderzeugungselementes; (3) nach der Stufe (2), Aussetzen des geladenen Bilderzeugungselementes aktivierender Strahlung bei einer Wellenlänge, für welche das Migrationsmarkierungsmaterial empfindlich ist; (4) nach Stufe (3), Bewirken der Erweichung des erweichbaren Materials und Befähigen eines ersten Teiles des Migrationsmarkierungsmaterials, durch das erweichbare Material zu dem Substrat in einem bildweisen Muster zu migrieren, während ein zweiter Teil des Migrationsmarkierungsmaterials im wesentlichen nicht migriert in der erweichbaren Schicht zurückbleibt; worin nach der Migration des ersten Teiles des Migrationsmarkierungsmaterials entweder (a) der erste Teil des Migrationsmarkierungsmaterials das transparentmachende Mittel kontaktiert und der zweite Teil des Migrationsmarkierungsmaterials das transparentmachende Mittel nicht kontaktiert; oder (b) der zweite Teil des Migrationsmarkierungsmaterials das transparentmachende Mittel kontaktiert und der erste Teil des Migrationsmarkierungsmaterials das transparentmachende Mittel nicht kontaktiert.

10. Ein Verfahren nach Anspruch 9, worin der erste Teil des Migrationsmarkierungsmaterials das transparentmachende Mittel kontaktiert und der zweite Teil des Migrationsmarkierungsmaterials das transparentmachende Mittel nicht kontaktiert; oder worin der zweite Teil des Migrationsmarkierungsmaterials das transparentmachende Mittel kontaktiert und der erste Teil des Migrationsmarkierungsmaterials das transparentmachende Mittel nicht kontaktiert.

## Revendications

1. Elément de formation d'images par migration (1) comprenant (a) un substrat (2), (b) une couche ramollissable (6) comprenant un matériau ramollissable (7) et un matériau de marquage par migration photosensible (8), et (c) un agent de transparence qui rend transparent le matériau de marquage par migration en contact avec lui, contenu dans au moins une couche de l'élément de formation d'images par migration, dans lequel l'agent de transparence agit sur le matériau de marquage par migration qui entre en contact avec lui en réduisant la densité optique de la couche ramollissable contenant le matériau de marquage par migration.

2. Elément de formation d'images par migration selon la revendication 1, dans lequel le matériau de marquage par migration (8) est choisi dans le groupe constitué par (a) le sélénium, (b) le tellure, (c) des alliages de sélénium et d'un matériau choisi dans le groupe constitué par le tellure, l'arsenic, l'antimoine, le thallium, le bismuth, ou des mélanges de ceux-ci, (d) des alliages de tellure et d'un matériau choisi dans le groupe constitué par l'arsenic, l'antimoine, le thallium, le bismuth ou des mélanges de ceux-ci, (e) du sélénium dopé par un halogène, (f) du tellure dopé par un halogène, (g) des alliages dopés par un halogène de sélénium et d'un matériau choisi dans le groupe constitué par le tellure, l'arsenic, l'antimoine, le thallium, le bismuth ou des mélanges de ceux-ci, (h) des alliages dopés par un halogène de tellure et d'un matériau choisi dans le groupe constitué par l'arsenic, l'antimoine, le thallium, le bismuth ou des mélanges de ceux-ci, et (i) des mélanges de ceux-ci.

3. Elément de formation d'images par migration selon la revendication 1 ou la revendication 2, dans lequel l'agent de transparence est contenu dans la couche ramollissable.

4. Elément de formation d'images par migration selon la revendication 1 ou la revendication 2, dans lequel l'agent de transparence est contenu dans une couche située entre la couche ramollissable et le substrat.

5. Elément de formation d'images par migration selon la revendication 1 ou 2, dans lequel la couche ramollissable est située entre le substrat et une couche contenant l'agent de transparence.

6. Elément de formation d'images par migration selon la revendication 1 ou la revendication 2, dans lequel l'élément de formation d'images par migration comprend un substrat, une première couche ramollissable comprenant un premier matériau ramollissable et un premier matériau de marquage par migration, et une seconde couche ramollissable comprenant un second matériau ramollissable et un second matériau de marquage par migration, dans lequel l'agent de transparence est contenu dans une couche située entre la première couche ramollissable et la seconde couche ramollissable.

7. Elément de formation d'images par migration selon l'une quelconque des revendications 1 à 6, dans lequel l'agent de transparence est présent en une quantité d'environ 1 à environ 50 % en poids du matériau constituant la couche dans laquelle il est contenu.

8. Elément de formation d'images par migration selon la revendication 1, dans lequel l'agent de transparence est un composé azacyclique ; ou dans lequel l'agent de transparence est choisi dans le groupe constitué par : (A) des matériaux répondant aux formules générales : dans lesquelles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈ et R₃₉ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, R₂₈, R₂₉, R₃₀, R₃₁, R₃₂, R₃₃, R₃₄, R₃₅, R₃₆, R₃₇, R₃₈ et R₃₉ peuvent être liés ensemble pour former un cycle ; (B) des matériaux répondant aux formules générales : dans lesquelles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ et R₂₂ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁ et R₂₂ peuvent être liés ensemble pour former un cycle ; (C) des matériaux répondant aux formules générales : dans lesquelles R₁, R₂, et R₃ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂ et R₃ peuvent être liés ensemble pour former un cycle ; (D) des matériaux répondant aux formules générales : dans lesquelles R₁, R₂, R₃, R₄, R₅, R₆, R₇, R₈, R₉, R₁₀, R₁₁, R₁₂, sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂, R₃, R₄, R₅, R₆, R₇, R₈, R₉, R₁₀, R₁₁ et R₁₂ peuvent être liés ensemble pour former un cycle ; (E) des matériaux répondant aux formules générales : dans lesquelles R₁, R₂, R₃, et R₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂, R₃, et R₄ peuvent être liés ensemble pour former un cycle ; (F) des matériaux répondant à la formule générale dans laquelle R₁, R₂, R₃, R₄, R₅, R₆, R₇, R₈, R₉, R₁₀, R₁₁, R₁₂, R₁₃ et R₁₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, R₄, R₅, R₆, R₇, R₈, R₉, R₁₀, R₁₁, R₁₂, R₁₃ et R₁₄ peuvent être liés ensemble pour former un cycle ; (G) des matériaux répondant à la formule générale : dans laquelle R₁ et R₂ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquels deux ou plus de deux des symboles R₁, et R₂ peuvent être liés ensemble pour former un cycle ; (H) des matériaux répondant à la formule générale : dans laquelle R₁, R₂, R₃, R₄, et R₆ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, R₄, et R₅ peuvent être liés ensemble pour former un cycle ; (I) des matériaux répondant à la formule générale : dans laquelle R₁, R₂, R₃, R₄, R₅, R₆, R₇, R₈ et R₉ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, R₄, R₅, R₆, R₇, R₈ et R₉ peuvent être liés ensemble pour former un cycle ; (J) des matériaux répondant à la formule générale : dans laquelle R₁, R₂, R₃, et R₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, et R₄ peuvent être liés ensemble pour former un cycle ; (K) des matériaux répondant à la formule générale : dans laquelle R₁, R₂, R₃, et R₄, sont choisis, chacun indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, et R₄ peuvent être liés ensemble pour former un cycle ; (L) des matériaux répondant à la formule générale : dans laquelle R₁, R₂, R₃, R₄ et R₅ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, R₄ et R₅ peuvent être liés ensemble pour former un cycle ; (M) des matériaux répondant aux formules générales : dans lesquelles R₁, R₂, R₃, R₄, R₅, R₆, R₇, R₈, R₉, R₁₀, R₁₁, R₁₂, R₁₃ et R₁₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans lesquelles deux ou plus de deux des symboles R₁, R₂, R₃, R₄, R₅, R₆, R₇, R₈, R₉, R₁₀, R₁₁, R₁₂, R₁₃ et R₁₄ peuvent être liés ensemble pour former un cycle ; (N) des matériaux répondant à la formule générale : dans laquelle R₁, R₂, R₃, et R₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, et R₄ peuvent être liés ensemble pour former un cycle ; (O) des matériaux répondant à la formule générale : dans laquelle R₁, R₂, R₃, et R₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, et R₄ peuvent être liés ensemble pour former un cycle ; (P) des matériaux répondant à la formule générale : dans laquelle R₁, R₂, R₃, et R₄ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃, et R₄ peuvent être liés ensemble pour former un cycle ; (Q) des matériaux répondant à la formule générale : dans laquelle R₁, R₂, R₃ et R₄ sont choisis chacun, indépendamment des autres, dans le groupe constitué par des atomes d'hydrogène, des groupes alkyle, des groupes aklyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, dans laquelle deux ou plus de deux des symboles R₁, R₂, R₃ et R₄ peuvent être liés ensemble pour former un cycle ; (R) des matériaux répondant aux formules générales : dans laquelle R₁ est choisi dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide et dans lesquelles la partie courbe de la structure représente une chaîne hydrocarbonée ou une chaîne hydrocarbonée substituée, dans lesquelles deux ou plus de deux substituants peuvent être liés ensemble pour former un cycle ; (S) des matériaux répondant à la formule générale : dans laquelle R₁ est choisi dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide, et des groupes azide, et dans laquelle la partie courbe de la structure représente une chaîne hydrocarbonée ou une chaîne hydrocarbonée substituée, dans laquelle deux ou plus de deux substituants peuvent être liés ensemble pour former un cycle ; (T) des mélanges de ceux-ci ; ou dans lequel l'agent de transparence est choisi dans le groupe constitué par l'homopipéridine, (2) le thiocyanate de pipéridine, (3) le 2-pipéridineméthanol, (4) le 3-pipéridineméthanol, (5) le 2-pipéridineéthanol, (6) le 4-pipéridineéthanol, (7) le monohydrate de chlorhydrate de 4-pipéridine, (8) la 1-aminopipéridine, (9) la 1-(2-aminoéthyl)pipéridine, (10) la 4-(aminométhyl)pipéridine, (11) le 3-pipéridino-1,2-propanediol (Aldrich 21,849-9), (12) l'acide 1-pipéridinepropionique, (13) la 1-méthyl-4(méthylamino)pipéridine, (14) la 1-acétyl-3-méthylpipéridine, (15) la 4'-pipéridinoacétophénone, (16) la 4-phénylpipéridine, (17) la 4-pipéridinopipéridine, (18) la 4-benzylpipéridine, (19) la 4-(4-méthylpipéridino)pyridine, (20) le 4-pipéridoneéthylèneacétal, (21) la bis(pentaméthylène)urée, (22) la 1- benzyl-4-hydroxypipéridine, (23) la 1-benzoyl-4-pipéridone, (24) la 1,1'-méthylènebis (3-méthylpipéridine), (25) la 4,4'-triméthylènedi-pipéridine, (26) la 4,4'-triméthylènebis(1-menthylpipéridine), (27) le 4-4'-triméthylènebis(1-pipéridinepropionitrile), (28) le 4,4'-triméthylènebis-(1-pipéridineéthanol), (29) la 2,2,6,6-tétraméthylpipé-ridine, (30) la 4-amino-2,2,6,6-tétraméthylpipéridine, (31) la 4-(diméthylamino)-1,2,2,6,6-pentaméthyl-pipéridine, (32) la N,N'-bis-(2,2,6,6-tétraméthyl-4-pipéridinyl)-1,6-hexanediamine, (33) l'oxyde de tripipéridinophosphine, (34) le tropane, (35) l'hydrate de tropine, (36) la tropinone, (37) la 8-hydroxytropinone, (38) l'acide 2-pipéridinecarboxylique, (39) la 2-pipéridone, (40) le 4,4'-triméthylènebis(1-pipéridinecarboxamide), (41) le 4-méthyl-2-(pipéridinométhyl)phénol, (42) le bis-(chlorophénoxy)acétate de 1-méthyl-4-pipéridinyle, (43) le monochlorhydrate de chlorure de 2-(hexaméthylène-imino)éthyle, (44) le chlorhydrate de 3-(hexahydro-1H-azépin-1-yl)-3'-nitropropiophénone, (45) le chlorhydrate d'imipramine, (46) la carbamézépine, (47) le chlorhydrate de 5,6,11,12-tétrahydrodibenz[b,f]azocine, (48) le chlorhydrate de quinuclidine, (49) le chlorhydrate de 3-quinuclidinol, (50) le chlorhydrate de 3-quinuclidinone, (51) le dihydrate de chlorhydrate de 2-méthylène-3-quinuclidinone, (52) le dichlorhydrate de 3-aminoquinuclidine, (53) le chlorhydrate de 3-chloro-quinuclidine, (54) le dihydrate de sulfate de quinidine, (55) le dihydrate de monochlorhydrate de quinine, (56) le monohydrate de sulfate de quinine, (57) le chlorhydrate d'hydroquinidine, (58) le dihydrate de bromhydrate d'hydroquinine, (59) la pipérazine, (60) l'homopipérazine, (61) la 1-méthylpipérazine, (62) la 2-méthylpipérazine, (63) la 1-acétylpipérazine, (64) la 1-(2-hydroxyéthyl)pipérazine, (65) la 1-(2-aminoéthyl)pipérazine, (66) le 1-pipérazinecarboxylate de tert-butyle, (67) le N-isopropyl-1-pipérazineacétamide, (68) la 1-(2-méthoxyphényl)pipérazine, (69) la 1-(2-pyridyl)pipérazine, (70) la 1-benzylpipérazine, (71) la 1-cinnamylpipérazine, (72) la 1-(4-chlorobenzhy-dryl)pipérazine, (73) la 2,6-diméthylpipérazine, (74) la 1-amino-4-méthylpipérazine, (75) la 1-amino-4-(2-hydroxyéthyl)-pipérazine, (76) la 1,4-bis(2-hydroxyéthyl)pipérazine, (77) la 1,4-bis(3-aminopropyl)-pipérazine, (78) le carboxylate de tert-butyl-4-benzyl-1-pipérazine, (79) la 1-pipéronylpipérazine, (80) le disulfure de bis(4-méthyl-1-homopipérazinyl-thiocarbonyle), (81) le monohydrate de dichlorhydrate de 1-amino-4-méthylpipérazine, (82) le monohydrate de dichlorhydrate de 1-(3-chloropropyl)-pipérazine, (83) le monochlorhydrate de 1-(2,3-xylyl)-pipérazine, (84) l'iodure de 1,1-diméthyl-4-phénylpipérazinium, (85) le 1,4,7-triazacyclononane, (86) le 1,5,9-triazacyclododécane, (87) le 1,2,3-triazole, (88) le 4-amino-1,2,4-triazole, (89) le 3-amino-5-méthylthio-1H-1,2,4-triazole, (90) le benzotriazole, (91) le 1-aminobenzotriazole, (92) le 1-cyanobenzotriazole, (93) le 5-méthyl-1H-benzotriazole, (94) l'isocyanure de 1H-benzotriazole-1-ylméthyle, (95) le méthacrylate de 2-[3-(2H-benzotriazole-2-yl)-4-hydroxyphényl]éthyle, (96) le 1,2,4-triazole, (97) le dérivé de sodium de 1,2,4-triazole, (98) le 3-amino-1,2,4-triazole, (99) le 3,5-diamino-1,2,4-triazole, (100) le 3-amino-5-mercapto-1,2,4-triazole, (101) l'hémihydrate de l'acide 3-amino-1,2,4-triazole-5-carboxylique, (102) le 4-amino-3-hydrazino-5-mercapto-1,2,4-triazole, (103) le monohydrate de l'acide 1,2,3-triazole-4,5-dicarboxylique, (104) le nitron, (105) l'hydrate de 1-hydroxybenzotriazole, (106) la 1,3,5-triazine, (107) l'acide cyanurique, (108) l'acide trithiocyanurique, (109) la 2,4-bis(méthylthio)-6-chloro-1,3,5-triazine, (110) la 2-chloro-4,6-diméthoxy-1,3,5-triazine, (111) la 2-chloro-4,6-diamino-1,3,5-triazine, (112) la trichloromélamine, (113) le chlorure cyanurique, (114) la 2,4,6-tris(perfluoroheptyl)-1,3,5-triazine, (115) le trihydrate d'hexahydro-2,4,6-triméthyl-1,3,5-triazine, (116) la 1,3,5-triméthylhexahydro-1,3,5-triazine, (117) la 1,3,5-triéthylhexahydro-1,3,5-triazine, (118) la 1,3,5-trichlohexylhexahydro-1,3,5-triazine, (119) la 1,3,5-tribenzylhexahydro-1,3,5-triazine, (120) l'acide trichloroisocyanurique, (121) le tris(isocyanurate de 2,3-dibromopropyle), (122) un composé d'acide cyanurique et de mélamine (123) l'urazole, (124) le 1-méthylurazole, (125) le 4-phénylurazole, (126) la 5-(4-hydroxyphényl)-5-phénylhydantoïne, (127) la β-tétralonehydantoïne, (128) le cyclène (1,4,7,10-tétraazacyclododécane), (129) le 1,4,8,11-tétraazacyclotétradécane, (130) le 1,4,8,11-tétraméthyl-1,4,8,11-tétraazacyclotétradécane, (131) la 1,4,8,11-tétraazacyclotétradécane-5,7-dione, (132) le 1,4,8,12-tétraazacyclopentadécane, (133) la 2,3,7,8,12,13,17,18-octaéthyl-21H,23H-porphine, (134) le 3,7,12,17-tétraméthyl-21H,23H-porphine-2,18-dipropionate de diméthyle, (135) le 7,12-diacétyl-3,8,13,17-tétraméthyl-21H,23H-porphine-2,18-dipropionate de diméthyle, (136) le sel disodique de l'acide 8,3-divinyl-3,7,12,17-tétraméthyl-21H,23H-porphine-2,18-dipropionique, (137) la 5,10,15,20-tétraphényl-21H,23H-porphine, (138) la 5,10,15,20-tétrakis(4-méthoxyphényl)-21H,23H-porphine, (139) le sel tétra-p-tosylate de 5,10,15-20-tétrakis[4-(triméthylamino)phényl]-21H,23H-porphine, (140) la 5,10,15,20-tétra(4-pyridyl)-21H,23H-porphine, (141) le sel tétra-p-tosylate de 5,10,15,20-tétrakis(1-méthyl-4-pyridyl)-21H,23H-porphine, (142) le 1,5-pentaméthylènetétrazole, (143) le 1-H-tétrazole, (144) le monohydrate de 5-aminotétrazole, (145) le chlorure de 2,3,5-triphényl-2H-tétrazolium, (146) le chlorure de 2-(4-iodophényl)-5-(4-nitrophényl)-3-phényltétrazolium, (147) l'iodure de 1,2,3,3-tétraméthyl-3H-indolinium, (148) le trisulfate d'hexacyclène, (149) l'hexaméthylhexacyclène, (150) le pyrrole-2-carboxaldéhyde, (151) le prolineamide, (152) le 3-pyrrolidino-1,2-propanediol, (153) la 1-(pyrrolidinocarbonylméthyl)pipérazine, (154) la 4-pyrrolidinopyridine, (155) le 3-indolylacétonitrile, (156) la 6-nitroindoline, (157) le 7-azaindole, (158) l'indazole, (159) le 2-acétylpyrrole, (160) le 2-acétyl-1-méthylpyrrole, (161) le 3-acétyl-1-méthylpyrrole, (162) le 3-acétyl-2,4-diméthylpyrrole, (163) l'acide pyrrole-2-carboxylique, (164) l'acide 3-carboxy-1,4-diméthyl-2-pyrroleacétique, (165) la proline, (166) l'acide 2-pyrrolidone-5-carboxylique, (167) la 4-hydroxyproline, (168) l'acide 1,1'-éthylènebis(5-oxo-3-pyrrolidinecarboxylique, (169) le monohydrate de l'acide kaïnique, (170) le chlorohydrate de 1-aminopyrrolidine, (171) le chlorhydrate de 2-(2-chloroéthyl)-1-méthylpyrrolidine, (172) le chlorhydrate de 1-(2-chloroéthyl)pyrrolidine, (173) le dichlorhydrate de trémorine, (174) le chlorhydrate de l'ester méthylique de la L-proline, (175) le pyrrolidinedithiocarbamate d'ammonium, (176) le tribromhydrate de pyrrolidone, (177) le chlorhydrate de 1-(4-chlorobenzyl)-2-(1-pyrrolidinylméthyl)benzimidazole, (178) le dichlorhydrate de billiverdine, (179) l'indole, (180) le 4,5,6,7-tétrahydroindole, (181) l'hydrate de 3-indoleméthanol, (182) le 3-indoleéthanol, (183) l'indole-3-carboxaldéhyde, (184) l'acétate de 3-indolyle, (185) l'indole-3-acétamide, (186) l'acide indole-3-carboxylique, (187) l'acide indole-3-acétique, (188) l'acide 3-indolepropionique, (189) l'acide 3-indoleacrylique, (190) l'acide 3-indoleglyoxylique, (191) l'acide indole-3-pyruvique, (192) l'acide 3-indolelactique, (193) l'acide 3-indolebutyrique, (194) le N-acétyltryptophanamide, (195) la N-(3-indolylacétyl)alanine, (196) la N-(3-indolylacétyl)valine, (197) la N-(3-indolylacétyl)isoleucine, (198) la N-(3-indolylacétyl)leucine, (199) l'acide N-(3-indolyl-acétyl)aspartique, (200) la N-(3-indolylacétyl)-L-phénylalanine, (201) le 4-hydroxyindole, (202) l'acide indole-4-carboxylique, (203) l'acétate de 4-indolyle, (204) le 4-méthylindole, (205) le 5-hydroxyindole, (206) l'acide 5-hydroxyindole-3-acétique, (207) l'acide 5-hydroxy-2-indolecarboxylique, (208) la N-acétyl-5-hydroxytryptamine, (209) l'acide indole-5-carboxylique, (210) le 5-méthylindole, (211) le 5-méthoxyindole, (212) l'acide indole-2-carboxylique, (213) l'acide indolène-2-carboxylique, (214) l'indole-2,3-dione, (215) le 2-méthylindole, (216) la 2,3,3-triméthylindolénine, (217) le chlorhydrate de tryptamine, (218) le chlorhydrate de 5-méthyltryptamine, (219) l'hémihydrate de chlorhydrate de sérotonine, (220) le monohydrate de chlorhydrate de norharmane, (221) le monohydrate de chlorhydrate d'harmane, (222) l'hydrate de chlorhydrate d'harmine, (223) l'hydrate de chorhydrate d'harmaline, (224) le dihydrate de chlorhydrate d'harmol, (225) le dihydrate de chlorhydrate d'harmalol, (226) le chlorhydrate de 3,6-diaminoacridine, (227) l'iodure de (3-indolyl)isothiuronium, (228) le chlorhydrate de yohimbine, (229) le pyrazole, (230) le 3-aminopyrazole, (231) le 5-amino-1-éthylpyrazole, (232) le 3-amino-4-carbéthoxypyrazole, (233) le 3-amino-5-méthylpyrazole, (234) le 3-amino-5-phénylpyrazole, (235) le 4-pyrazolecarboxylate d'éthyle, (236) le 3,5-pyrazolecarboxylate de diéthyle, (237) le 1,1'-(1-éthylpropylidène)bis-lH-pyrazole, (238) le 4-bromopyrazole, (239) le 4-bromo-3-méthylpyrazole, (240) le 3,5-diméthylpyrazole, (241) le 4-bromo-3,5-diméthylpyrazole, (242) le 3,5-diméthylpyrazole-1-carboxamide, (243) le 3,5-diméthylpyrazole-1-méthanol, (244) le 3-méthyl-1-vinylpyrazole, (245) la 4-benzoyl-3-méthyl-1-phényl-2-pyrazolin-5-one, (246) le 1-nitropyrazole, (247) l'acide 4-pyrazolecarboxylique, (248) le monohydrate de l'acide 3,5-pyrazoledicarboxylique, (249) le 3-amino-5-hydroxypyrazole, (250) le 3-amino-4-pyrazolecarbonitrile, (251) l'acide 3-amino-4-pyrazolecarboxylique, (252) le chlorhydrate de 4-méthylpyrazole, (253) le sulfate de 3,4-diamino-5-hydroxypyrazole, (254) le nitrate de 3,5-diméthylpyrazole-1-carboxamidine, (255) l'hémisulfate de 3-amino-4-pyrazolecarboxamide, (256) un sel d'acide du chlorhydrate de 6-aminoindazole, (257) la 4-hydroxypyrazolo[3, 4-d]pyrimidine, (258) la 4-mercapto-lH-pyrazolo-[3,4-d]-pyrimidine, (259) l'indazole, (260) le 5-aminoindazole, (261) le 6-aminoindazole, (262) la 3-indazolinone, (263) le N'-(6-indazolyl)sulfanilamide, (264) le méthanesulfonate de 4,5-dihydro-3-(4-pyridinyl)-2H-benz[g]indazole, (265) l'imidazole, (266) le 4-méthylimidazole, (267) le 2-éthylimidazole, (268) le 2-propylimidazole, (269) le 1-butylimidazole, (270) le 2-undécylimidazole, (271) l'histamine, (272) le 1-(3-aminopropyl)imidazole, (273) le 1-acétylimidazole, (274) le 2-méthyl-1-vinylimidazole, (275) le 2-éthyl-4-méthylimidazole, (276) le 1-benzyl-2-méthylimidazole, (277) le 1-méthylbenzimidazole, (278) le chlorure de 1-éthyl-3-méthyl-1,H-imidazolinium, (279) l'hydrate de dichlorhydrate de 2-(aminométhyl)benzimidazole, (280) le monohydrate d'hémisulfate de 2,6-diamino-8-purinol, (281) le chlorure de purin-6-yl-triméthylammonium, (282) le chlorhydrate de 4-méthyl-5-imidazoleméthanol, (283) le dipropanoate de N,N'-bis[3-(4,5-dihydro-1H-imidazol-2-yl)phényl]urée, (284) l'iodure de 1-(p-tosyl)-3,4,4-triméthyl-2-imidazolinium, (285) le chlorure de 1-éthyl-3-méthyl-1H-imidazolinium, (286) le sulfate de 2-aminoimidazole, (287) le chlorhydrate de 4-amino-5-imidazolecarboxamide, (288) le bromhydrate de 2-hydrazino-2-imidazoline, (289) le chlorhydrate d'imidazole, (290) le chlorhydrate d'acide 4-imidazole-acétique, (291) le chlorhydrate de 2-benzyl-2-imidazoline, (292) le chlorhydrate de 1-(1-phényl-éthyl)imidazole-5-carboxylate de propyle, (293) l'hydrate de sulfate de 2,6-diaminopurine, (294) le méthylsulfate de 1-suif-amidoéthyl-3-méthyl-2-heptadécylimidazolinium, (295) l'éthylsulfate d'isostéaryléthylimidonium, (296) le méthylsulfate de méthyl-1-suif-amidoéthyl-2-suif-imidazolinium, (297) le chlorure d'isostéarylbenzylimidonium, (298) le méthyl-1-suif hydrogéné-amidoéthyle, (299) le méthylsulfate de suif hydrogéné-imidazolinium, (300) le méthylsulfate de 1-méthyl-1-oléylamidoéthyl-2-oléylimidazolinium, (301) le chlorure de phosphate de cocohydroxyéthylpolyéthylèneglycolimidazolinium, (302) la guanine, (303) l'hydrate de guanosine, (304) la xanthine, (305) la 1-méthylxanthine, (306) la 3-méthylxanthine, (307) la 3-isobutyl-1-méthylxanthine, (308) l'hypoxanthine, (309) le dihydrate de xanthosine, (310) le 6-thioxanthène, (311) la purine, (312) la 6-aminopurine, (313) l'hémihydrate de 6-méthoxypurine, (314) le monohydrate de 6-mercaptopurine, (315) la 2-amino-6-chloropurine, (316) la 2-amino-6,8- dihydroxypurine, (317) la théophylline (3,7-dihydro-1,3-diméthyl-1H-purine-2,6-dione), (318) la kinétine, (319) la 1-méthyladénine, (320) la 3-méthyladénine, (321) l'adénosine, (322) l'inosine, (323) le 6-mercaptopurineriboside, (324) l'hémihydrate de chlorhydrate de 6-aminopurine, (325) le sulfate de 6-aminopurine, (326) le monohohydrate d'hémisulfate de 2,6-diamino-8-purinol, (327) le benzimidazole, (328) le 2-aminobenzimidazole, (329) le 2-amino-5,6-diméthylbenzimidazole, (330) l'acide 5-benzimidazolecarboxylique, (331) le 2,4,5-triméthylbenzimidazole, (332) le 2-guanidinobenzimidazole, (333) le 2-hydroxybenzimidazole, (334) la 4-(2-céto-1-benzimidazolinyl)pipéridine, (335) la 2-imidazolidinethione, (336) la 2-imidazolidone, (337) l'hydantoïne, (338) la 1-méthylhydantoïne, (339) la créatinine, (340) la 2-thiohydantoïne, (341) l'acide 5-hydantoïneacétique, (342) la 5-uréidohydantoïne, (343) la 5,5-diméthylhydantoïne, (344) l'acide 2-imidazolidone-4-carboxylique, (345) le N,N-bis(2-hydroxyéthyl)isonicotinamide, (346) le 1,2-bis(4-pyridyl)éthylène, (347) la 2-(2-pipéridinoéthyl)pyridine, (348) le 1,2-bis(4-pyridyl)éthane, (349) la 4,4'-triméthylènepyridine, (350) l'aldrithiol-2, (351) l'aldrithiol-4, (352) la 1,3-bis(3-pyridylméthyl)-2-thiourée, (353) la 2,2' : 6',2" -terpyridine, (354) la 2-[N,N-bis(trifluorométhylsulfonyl)amino]pyridine, (355) l'acide 2,3-pyridinedicarboxylique, (356) le monohydrate d'acide 2,4-pyridinedicarboxylique, (357) l'acide 2,5-pyridinedicarboxylique, (358) l'acide 2,6-pyridinedicarboxylique, (359) l'acide 3,4-pyridinedicarboxylique, (360) l'acide 3,5-pyridinedicarboxylique, (361) le 2,6-pyridinedicarboxaldéhyde, (362) le 3,4-pyridinecarboxamide, (363) le 3,4-pyridinecarboximide, (364) l'anhydride 2,3-pyridinecarboxylique, (365) l'anhydride 3,4-pyridinecarboxylique, (366) le 2,6-pyridineméthanol, (367) l'acide 2-pyridineéthanesulfonique, (368) l'acide 4-pyridineéthanesulfonique, (369) l'acide 3-pyridinesulfonique, (370) l'acide pyridoxique, (371) l'acide trans-3-(3-pyridyl)acrylique, (372) l'acide 2-pyridylhydroxyméthanesulfonique, (373) l'acide 3-pyridylhydroxyméthanesulfonique, (374) l'acide 6-méthyl-2,3-pyridinedicarboxylique, (375) l'acide isonicotinique, (376) le bromhydrate de pyridine, (377) le chlorhydrate de pyridine, (378) le chlorhydrate de 2-(chlorométhyl)pyridine, (379) le chlorhydrate d'acide 2-pyridylacétique, (380) le chlorhydrate de chlorure de nicotinoyle, (381) le dichlorhydrate de 2-hydrazinopyridine, (382) le dichlorhydrate de 2-(2-méthylaminoéthyl)pyridine, (383) le chlorhydrate de 1-méthyl-1,2,3,6-tétrahydropyridine, (384) le chlorhydrate de 2,6-dihydroxypyridine, (385) le chlorhydrate de 3-hydroxy-2(hydroxyméthyl)pyridine, (386) le chlorhydrate de pyridoxine, (387) le chlorhydrate de pyridoxal, (388) le monohydrate de 5-phosphate de pyridoxal, (389) le chlorhydrate de 3-amino-2,6-diméthoxypyridine, (390) le monohydrate de dichlorhydrate de pyridoxamine, (391) le phosphate d'iproniazide, (392) le chlorhydrate de tripélennamine, (393) le perbromure de bromure de pyridinium, (394) le 3-nitrobenzènesulfonate de pyridinium, (395) le bromure de 1-éthyl-3-hydroxy-pyridinium, (396) l'iodure de 1-éthyl-4-(méthoxy-carbonyl)pyridinium, (397) le bromure de 1-heptyl-4-(4-pyridyl)pyridinium, (398) le chlorure de 1-dodécylpyridinium, (399) le monohydrate de chlorure de 1-hexadécylpyridinium, (400) le monohydrate de bromure de 1-hexadécylpyridinium, (401) le chlorure de 1-(carboxyméthyl)pyridinium, (402) l'hydrazide de chlorure de 1-(carboxyméthyl)pyridinium, (403) le chlorure de 1-(3-nitrobenzyloxyméthyl)pyridinium, (404) l'hydroxyde de 1-(3-sulfopropyl)pyridinium, (405) le chlorure de N-(lauroylcolaminoformylméthyl)pyridinium, (406) le chlorure de N-(stéaroylcolamineformylméthyl)pyridinium, (407) l'iodure de 2-chloro-1-méthylpyridinium, (408) le méthanesulfonate de 2-pyridinealdoxime-l-méthyle, le chlorure de 2-pyridinealdoxime-1-méthyle, (409) l'iodure de 2-[4-(diméthylamino)styryl]-1-éthylpyridinium, (410) le chlorure de 1-benzyl-3-hydroxypyridinium, (411) l'iodure de 1,4-diméthylpyridinium, (412) l'iodoure de 1-éthyl-4-phénylpyridinium, (413) l'iodure de 4-phényl-1-propylpyridinium, (414) le bromure de 1-docosyl-4-(4-hydroxystyryl)pyridinium, (415) le dichlorure de 1,1'-diméthyl-4-4'-bipyridinium, (416) le dibromure de 1,1'-diéthyl-4-4'-bipyridinium, (417) le dichlorure de 1,1'-dibenzyl-4,4'-bipyridinium, (418) le dibromure de 1,1'-diheptyl-4,4'-bipyridinium, (419) la 1,7-phénanthroline, (420) la 1,10-phénanthroline, (421) la 5-chloro-1,10-phénanthroline, (422) le méthanesulfonate de 4,5-dihydro-3-(4-pyridinyl)-2H-benz[g]indazole, (423) la 1,2,3,4-tétrahydroquinoléine, (424) la 6-éthoxy-1,2,3,4-tétrahydro-2,2,4-triméthylquinoléine, (425) la 2-cyanoquinoléine, (426) la 1-cyanoisoquinoléine, (427) la 3-cyanoisoquinoléine, (428) la 3-aminoquinoléine, (429) la 8-aminoquinoléine, (430) la 7,8-benzoquinoléine, (431) la 8-hydroxyquinoléine, (432) le sel d'aluminium de la 8-hydroxyquinoléine, (433) la 8-hydroxyquinaldine, (434) la 3,4,5,6,7,8-hexahydro-2-(1H)-quinolinone, (435) la julolidine, (436) la quinoxaline, (437) le 2-quinoxalinecarboxylate d'éthyle, (438) la quinoléine, (439) la 2-hydroxyquinoléine, (440) la 4-hydroxyquinoléine, (441) la 5-hydroxyquinoléine, (442) la 5-aminoquinoléine, (443) la 6-aminoquinoléine, (444) l'acide 2-quinoléinecarboxylique, (445) l'acide 3-quinoléinecarboxylique, (446) l'acide 4-quinoléinecarboxylique, (447) le 4-quinoléinecarboxaldéhyde, (448) le 2-quinoléinethiol, (449) le 2,4-quinoléinediol, (450) la quinaldine, (451) la 4-aminoquinaldine, (452) la 2,6-diméthylquinoléine, (453) la 2,7-diméthylquinoléine, (454) l'acide 4-méthoxy-2-quinoléinecarboxylique, (455) le 2-phényl-4-quinoléinecarboxylate de méthyle, (456) la 2-(N-butyl-carbamoyl)-1,2,3,4-tétrahydraisoquinoléine, (457) la 1-hydroxyisoquinoléine, (458) l'acide 1-isoquinoléinecarboxylique, (459) l'acide 3-isoquinoléinecarboxylique, (460) le 1,5-isoquinoléinediol, (461) l'hémihydrate d'hémisulfate de 8-hydroxyquinoléine, (462) le dichlorhydrate de 5-amino-8-hydroxyquinoléine, (463) le monochlorhydrate de 2-(chlorométhyl)quinoléïne, (464) le monohydrate d'acide 8-hydroxyquinoléine-5-sulfonique, (465) l'hydrate du sel de sodium de l'acide 8-éthoxy-5-quinoléinesulfonique, (466) le chlorhydrate de 1,2,3,4-tétrahydroisoquinoléine, (467) le chlorhydrate de l'acide 1,2,3,4-tétrahydro-3-isoquinoléinecarboxylique acide, (468) le chlorhydrate de 6,7-diméthoxy-1,2,3,4-tétrahydroisoquinoléine, (469) le bromhydrate de 1-méthyl-6,7-dihydroxy-1,2,3,4-tétrahydroisoquinoléine, (470) le diphosphate de primaquine, (471) le phosphate de pentaquine, (472) le chlorhydrate de dibucaïne, (473) l'hémihydrate de chlorhydrate de 9-aminoacridine, (474) l'hémisulfate de 3,6-diaminoacridine, (475) le chlorhydrate de 2-quinoléinethiol, (476) le pentahydrate de sulfate de spartéine, (477) le chlorhydrate de papavérine, (478) l'hydrate de dichlorhydrate d'émétine, (479) le monohydrate de monochlorhydrate de 1,10-phénanthroline, (480) le trihydrate de chlorhydrate de néocuproïne, (481) la pyrimidine, (482) la 2-chloropyrimidine, (483) la 4-phénylpyrimidine, (484) la 5-bromopyrimidine, (485) la 2,4-dichloropyrimidine, (486) la 4,6-dichloropyrimidine, (487) la 2,4-dichloro-6-méthylpyrimidine, (488) la 6-chloro-2,4-diméthoxypyrimidine, (489) la 2-amino-4,6-diméthoxypyrimidine, (490) la 2,4,6-trichloropyrimidine, (491) la 2,4,5,6-tétrachloropyrimidine, (492) la 1,3,4,6,7,8-hexahydro-1-méthyl-2H-pyrimido[1,2-a]pyrimidine, (493) la 1,3,4,6,7,8-hexahydro-2H-pyrimido-[1,2-a]pyrimidine, (494) l'hexétidine, (495) le S-(4,6-diméthylpyrimidin-2-yl)thiocarbonate de tert-butyle, (496) le S-(4,6-diméthylpyrimidin-2-yl)thiocarbonate de 4-méthoxybenzyle, (497) la 2-aminopyrimidine, (498) la 2-amino-4-méthylpyrimidine, (499) la 2-amino-5-nitropyrimidine, (500) la 2-amino-5-bromopyrimidine, (501) la 2-amino-4-chloro-6-méthylpyrimidine, (502) la 2-amino-4,6-diméthylpyrimidine, (503) la 2-amino-4-hydroxy-6-méthylpyrimidine, (504) la 2-amino-4,6-dichloropyrimidine, (505) le 2-amino-5-bromo-6-méthyl-4-pyrimidinol, (506) la 4-aminopyrimidine, (507) la 4,5-diaminopyrimidine, (508) la 4-amino-2,6-diméthylpyrimidine, (509) la 2,4-diamino-6-hydroxypyrimidine, (510) la 2,6-diamino-4-chloropyrimidine, (511) l'hémihydrate de 4,6-diamino-2-mercaptopyrimidine, (512) la 2,4,6-triaminopyridine, (513) la 5-nitroso-2,4,6-triaminopyrimidine, (514) la 4,6-dihydroxypyrimidine, (515) la 4,6-dihydroxy-2-aminopyrimidine, (516) la 4,6-dihydroxy-2-méthylpyrimidine, (517) la 4,6-dihydroxy-5-nitropyrimidine, (518) la 2,4-hihydroxy-5-méthylpyrimidine, (519) 2,4-dihydroxy-6-méthylpyrimidine, (520) la 2,4-dihydroxy-5,6-diméthylpyrimidine, (521) l'hydrate d'acide 2,6-dihydroxypyrimidine-5-carboxylique, (522) la 2,6-dihydroxy-4-aminopyrimidine, (523) la 2,4,5-trihydroxypyrimidine, (524) le 2-thiouracile, (525) le 6-amino-5-nitroso-2-thiouracile, (526) le dihydrate d'acide folique, (527) l'hydrate de sel de calcium d'acide folinique, (528) le chlorhydrate de 2-hydroxypyrimidine, (529) le chlorhydrate de 2-hydroxy-4-méthylpyrimidine, (530) le chlorhydrate de 4,6-diméthyl-2-hydroxypyrimidine, (531) le chlorhydrate de 2-mercapto-4-méthylpyrimidine, (532) le monohydrate d'hémisulfate de 4,6-diaminopyrimidine, (533) l'hydrate de sulfate de 4,5,6-triaminopyrimidine, (534) le sulfate de 4,5-diamino-6-hydroxypyrimidine, (535) l'hémisulfate de 2,4-diamino-6-mercaptopyrimidine, (536) l'hydrate d'hémisulfate de 2,4-diamino-6-hydroxypyrimidine, (537) le sulfate de 6-hydroxy-2,4,5-triaminopyrimidine, (538) le sulfate de 5,6-diamino-2,4-dihydroxypyrimidine, (539) le monochlorhydrate de N⁴-(2-amino-4-pyrimidinyl)sulfanilamide, (540) le sulfate de 2,4,5,6-tétraaminopyrimidine, (541) la 2,4-(1H,3H)-pyrimidinedione, (542) le 5-aminouracile, (543) le 5-nitrouracile, (544) le 5-iodouracile, (545) l'hydrate de 5-(hydroxyméthyl)uracile, (546) le 5,6-dihydrouracile, (547) le 6-amino-1-méthyluracile, (548) l'hydrate de 5,6-diamino-1,3-diméthyluracile, (549) l'uridine, (550) la 5-méthyluridine, (551) la 5-iodouridine, (552) la thimidine, (553) le 5-méthyl-2-thiouracile, (554) la 4-thiouridine, (555) le dihydrate de 2-thiocytidine, (556) le monohydrate d'acide orotique, (557) l'acide hydroorotique, (558) l'acide 5-aminoorotique, (559) l'orotate de méthyle, (560) l'acide barbiturique, (561) le trihydrate de l'acide 5-nitrobarbiturique, (562) le monohydrate de l'acide violurique, (563) le monohydrate d'alloxane, (564) le sulfate de 4,5,6-triamino-2(1H)-pyrimidinéthione, (565) le chlorhydrate de cyclocytidine, (566) le chlorhydrate de cytosinearabinoside, (567) la pyridazine, (568) la phtalazine, (569) le monohydrate de 4,5-dihydro-6-méthyl-3(2H)-pyridazinone, (570) la 3,6-dichloropyridazine, (571) la 3,4,5-trichloropyridazine, (572) la 3,6-dichloro-4-méthylpyridazine, (573) la 3-chloro-6-méthoxypyridazine, (574) la pyrazine, (575) l'acétylpyrazine, (576) l'aminopyrazine, (577) la 2,6-dichloropyrazine, (578) la 2,3,5-triméthylpyrazine, (579) la tétraméthylpyrazine, (580) l'acide 5-méthyl-2-pyrazinecarboxylique, (581) le pyrazineamide, (582) le 2,3-pyrazinedicarboxamide, (583) l'acide 4-pyridazinecarboxylique, (584) l'acide 2,3-pyrazinedicarboxylique, (585) le monohydrate de lumazine, (586) le monohydrate de xanthoptérine, (587) l'acide 2-quinoxazolinecarboxylique, (588) le 2-quinoxalinol, (589) la 2,3-dihydroxyquinoxaline, (590) le méthosulfate de phénazine, (591) la 2-azétidinone, (592) la 2-pyrrolidinone, (593) le tribromhydrate de pyrrolidone, (594) le δ-valérolactame, (595) l'ε-caprolactame, (596) l'amino-ε-caprolactame, (597) le N-méthylcaprolactame, (598) la 2-azacyclooctanone, (599) la 2-azacyclononanone, (600) l'ω-thiocaprolactame, (601) le N-vinylcaprolactame, (602) la 2-azabicyclo[2.2.1]hept-5-èn-3-one, (603) le maléimide, (604) le N-éthylmaléimide, (605) le N-butylmaléimide, (606) le N-cyclohexylmaléimide, (607) le N-phénylmaléimide, (608) le N-benzylmaléimide, (609) le N-hydroxymaléimide, (610) le succinimide, (611) le N-méthylsuccinimide, (612) le 2-hydroxy-N-méthylsuccinimide, (613) le N-hydroxysuccinimide, (614) le carbonate de succinimidyle et de 2,2,2-trichloroéthyle, (615) le 2-dodécyl-N-(2,2,6,6-tétraméthyl-4-pipéridinyl)succinimide, (616) le 2-dodécyl-N-(1,2,2,6,6-pentaméthyl-4-pipéridinyl)succinimide, (617) le N-(1-acétyl-2,2,6,6-tétraméthyl-4-pipéridinyl)-2-dodécylsuccinimide, (618) l'α-méthyl-α-propylsuccinimide, (619) l'α-méthyl-α-phénylsuccinimide, (620) le N-vinylphtalimide, (621) le N-éthylphtalimide, (622) le N-(triméthylsilylméthyl)phtalimide, (623) le N-(2-bromoéthyl)phtalimide, (624) le N-(3-bromopropyl)phtalimide, (625) le N-(4-bromobutyl)phtalimide, (626) le phtalimidoacétaldéhydediéthylacétal, (627) le (phtalimidométhyl)phosphonate de diéthyle, (628) le N-benzylphtalimide, (629) un sel de DBU (1,8-diazabicyclo[5.4.0]undéc-7-ène)-phtalimide (630) le DBN (1,5-diazabicyclo[4.3.0)]non-5-ène)-phtalimide et (631) des mélanges de ceux-ci ; ou dans lequel l'agent de transparence est un composé oxa-aza-cyclique ; ou dans lequel l'agent de transparence est choisi dans le groupe constitué par : (A) des matériaux répondant aux formules générales : dans lesquelles R₁, R₂, R₃, R₄, R₅, R₆, R₇, R₈, R₉, R₁₀, R₁₁, R₁₂, R₁₃, R₁₄ et R₁₅ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, R₁₀, R₁₁, R₁₂, R₁₃, R₁₄ et R₁₅ peuvent être liés ensemble pour former un cycle ; (B) des matériaux répondant à la formule générale : dans laquelle R₁, R₂, R₃, R₄, R₅, et R₆ sont choisis chacun, indépendamment des autres dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquels deux ou plus de deux des symboles R₁, R₂, R₃, R₄, R₅, et R₆ peuvent être liés ensemble pour former un cycle ; (C) des mélanges de ceux-ci ; ou dans lequel l'agent de transparence est choisi dans le groupe constitué par (1) le 3-amino-5-méthylisoxazole, (2) le 5-amino-3-méthylisoxazole, (3) le 3,5-diméthyl-4-nitroisoxazole, (4) le 1,2-benzisoxazole, (5) le 2,1-benzisoxazole, (6) la cyclosérine, (7) la 4-benzyl-2-méthyl-2-oxazoline, (8) le 2-méthyl-5-phényl-2-oxazoline-4-méthanol, (9) le benzoxazole, (10) le 2-méthylbenzoxazole, (11) le 2-chlorobenzoxazole, (12) le tétrafluoroborate de 2-chloro-3-éthylbenzeneoxazolium, (13) la 2-oxazolidone, (14) la 3-méthyl-2-oxazolidinone, (15) la 5-chlorométhyl-2-oxazolidinone, (16) la 4-isopropyl-2-oxazolidinone, (17) la 3-acétyl-2-oxazolidinone, (18) la 5,5-diméthyloxazolidine-2,4-dione, (19) la 3-éthyl-2-thioxo-4-oxazolidinone, (20) la 4-méthyl-5-phényl-2-oxazolidinone, (21) la 4-benzyl-2-oxazolidinone, (22) la 2-benzoisoxazolinone, (23) l'hydrate de muscimol, (24) l'acide 5-méthyl-3-phényl-isoxazole-4-çarboxylique, (25) le 2-méthyl-5-phényl-2-oxazoline-4-méthanol, (26) le sulfaméthoxazole, (27) le sulfisoxazole, (28) le N'-(4,5-diméthyloxazol-2-yl)sulfanilamide, (29) la chlorzoxazone, (30) l'iodure de 3,3'-diméthyloxacarbocyanine, (31) le 3'-sulfonate de 2-éthyl-5-phénylisoxazolium, (32) le perchlorate de 2-tert-butyl-5-méthylisoxazolium, (33) l'hydrate de chlorhydrate de 5-phényl-2-(4-pyridyl)oxazole, (34) le sel tosylate de méthyle de 5-phényl-2-(4-pyridyl)oxazole, (35) la 4-aminomorpholine, (36) le 4-morpholinecarbonitrile, (37) le 4-morpholinepropionitrile, (38) la 4-formylmorpholine, (39) la 4-acétylmorpholine, (40) la 4-(2-hydroxyéthyl)morpholine, (41) le 3-morpholino-1,2-propanediol, (42) la 4-(3-aminopropyl)morpholine, (43) le 1-morpholino-1-cyclopentène, (44) le 1-morpholino-1-cyclohexène, (45) le 1-morpholino-1-cycloheptène, (46) la 4-phénylmorpholine, (47) la 4-morpholinoaniline, (48) le phosphoromorpholinochloridate de 2,2,2-tribromoéthyle, (49) la 1-(morpholinocarbonylméthyl)pipérazine, (50) le 1,3-dimorpholine-2-nitropropane, (51) l'hémicholinium-3, (52) l'hémicholinium-15, (53) le chlorure de 2-méthoxy-4-morpholinobenzènediazonium, le chlorure de zinc, (54) la fomocaïne, (55) la 4-morpholinobenzophénone, (56) la 4,4'-éthylène-bis(2,6-morpholinedione), (57) la N,N'-dicyclohexyl-4-morpholinecarboxamidine, (58) la 1-cyclohexyl-3-(2-morpholinoéthyl)-2-thiourée, (59) la 4-morpholinoacétophénone, (60) le chlorhydrate de 4-(2-chloroéthyl)morpholine, (61) l'acide 4-morpholineéthanesulfonique, (62) l'acide 4-morpholinepropanesulfonique, (63) l'acide β-hydroxymorpholinepropanesulfonique, (64) le chlorhydrate de [N-(aminoiminométhyl)-4-morpholinecarboximidamide], (65) un composé d'acide 4-morpholinecarbodithioique et de morpholine, (66) le monohydrate du chlorhydrate de 2,5-diméthyl-4-(morpholinométhyl)phénol, (67) le méthop-toluènesulfonate de 1-cyclohexyl-3-(2-morpholinoéthyl)carbodiimide, (68) l'hémicholinium-3-[2,2'-(4,4'-biphènylène)bis(bromure de 2-hydroxy-4,4-diméthylmorpholinium]), (69) l'hémicholinium-15-[bromure de 4,4-diméthyl-2-hydroxy-2-phényl-morpholinium], (70) le 1-aza-12-couronne-4, (71) le 1-aza-15-couronne-5, (72) le 1-aza-18 couronne-6, (73) le 1,4,10-trioxa-7,13-diazacyclopentadécane, (74) le 1,4,10,13-tétraoxa-7,16-diazacyclooctadécane, (75) le N,N'-dibenzyl-1,4,10,13-tétraoxa-7,16-diazacyclooctadécane, (76) le 4,7,13,18-tétraoxa-1,10-diazabicyclo[8.5.5]éicosane, (77) le 4,7,13,16,21-pentaoxa-1,10-diazabicyclo[8.5.5]tricosane, (78) le 4,7,13,16,21,24-hexaoxa-1,10-diazabicyclo[8.8.8]hexacosane, (79) le 5,6-benzo-4,17,13,16,21,24-hexaoxa-1,10-diazabicyclo[8.8.8]hexacosane, et (80) des mélanges de ceux-ci ; ou dans lequel l'agent de transparence est un composé oxacyclique ; ou dans lequel l'agent de transparence est choisi dans le groupe constitué par : (A) des matériaux répondant à la formule générale : dans laquelle la partie courbe de la structure représente une chaîne hydrocarbonée ou une chaîne hydrocarbonée substituée, dans laquelle deux ou plus de deux substituants peuvent être liés ensemble pour former un cycle ; (B) des matériaux répondant aux formules générales : dans lesquelles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, et R₂₈ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, R₁₀, R₁₁, R₁₂, R₁₃, R₁₄, R₁₅, R₁₆, R₁₇, R₁₈, R₁₉, R₂₀, R₂₁, R₂₂, R₂₃, R₂₄, R₂₅, R₂₆, R₂₇, et R₂₈ peuvent être liés ensemble pour former un cycle ; (C) des matériaux répondant à la formule générale : dans laquelle la partie courbe de la structure représente une chaîne hydrocarbonée ou une chaîne hydrocarbonée substituée, dans laquelle deux ou plus de deux substituants peuvent être liés ensemble pour former un cycle ; (D) des matériaux répondant aux formules générales : dans lesquelles R₁, R₂, R₃, R₄, R₅, R₆, R₇, et R₈ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, et R₈ peuvent être liés ensemble pour former un cycle ; (E) des matériaux répondant aux formules générales : dans lesquelles les parties courbes des structures représentent une chaîne hydrocarbonée ou une chaîne hydrocarbonée substituée, dans lesquelles deux ou plus de deux substituants peuvent être liés ensemble pour former un cycle ; (F) des matériaux répondant à la formule générale : dans laquelle R₁, R₂, R₃, R₄, R₅, et R₆ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans laquelle deux ou plus de deux des symboles R₁, R₂, R₃, R₄, R₅, et R₆ peuvent être liés ensemble pour former un cycle ; et (G) des mélanges de ceux-ci ; ou dans lequel l'agent de transparence est choisi dans le groupe constitué par (1) la γ-butyrolactone, (2) la γ-valérolactone, (3) la γ-caprolactone, (4) la lactone γ-octanoïque, (5) la lactone γ-nonanoique, (6) la γ-décanolactone, (7) la γ-lactone undécanoïque, (8) la γ-phényl-γ-butyrolactone, (9) l'α-carbéthoxy-γ-phénylbutyrolactone, (10) la 2-coumaranone, (11) la β,β-diméthyl-γ-(hydroxyméthyl) -γ-butyrolactone, (12) la γ-éthoxycarbonyl-γ-butyrolactone, (13) la 5-(hydroxyméthyl)-2(5H)-furanone, (14) la dihydro-4,4-diméthyl-2,3-furandione, (15) la 2,5-diméthyl-4-hydroxy-3(2H)-furanone, (16) la (β-hydroxy-β-méthyl-δ-valéro)lactone mévalonique, (17) la δ-décanolactone, (18) la δ-lactone undécanoïque, (129) la δ-dodécanolactone, (20) la ω-lactone undécanoïque, (21) la oxacyclotridécan-2-one, (22) la ω-pentadécalactone, (23) l'hydrindantine (2,2'-dihydroxy-2,2'-biindan-1,1'3,3'-tétrone), (24) le dihydrate d'hydrindantine, (25) la 2-oxépanone, (26) la 4H-pyran-2-one, (27) le coumalate de méthyle, (28) le 2-oxo-2H-pyran-3-carboxylate de méthyle, (29) la 4,6-diméthyl-a-pyrone, (30) la 4-méthoxy-6-méthyl-2H-pyran-2-one, (31) la 3,6-dihydro-4,6,6-triméthyl-2H-pyran-2-one, (32) la 3,4-dihydro-6-méthyl-2H-pyran-2-one, (33) la 3-acétylcoumarine, (34) la 6-méthylcoumarine, (35) la 7-éthoxycoumarine, (36) le 3-coumarinecarboxylate d'éthyle, (37) la 7-diéthylamino-4-méthylcoumarine, (38) la dihydrocoumarine, (39) la 3-bromo-2-coumaranone, (40) la patuline, (41) la 4H-pyran-4-one, (42) la 2-éthyl-3-hydroxy-4H-pyran-4-one, (43) le butopyronoxyle (3,4-dihydro-2,2-diméthyl-4-oxo-2H-pyran-6-carboxylate de butyle, (44) l'acide déshydroacétique, (45) la 4-chromone, (46) la 4-chromanone, (47) le 4-chromanol, (48) la 6,7-diméthoxy-2,2-diméthyl-4-chromanone, (49) la 3-isochromanone, (50) la 6,7-diméthoxy-3-isochromanone, (51) le 6-éthyl-4-oxo-4H-1-benzopyran-3-carbonitrile, (52) le 6-éthyl-4-oxo-4H-1-benzopyran-3-carboxaldéhyde, (53) le 6-isopropyl-4-oxo-4H-1-benzopyran-3-carbonitrile, (54) le 6-isopropyl-4-oxo-4H-1-benzopyran-3-carboxaldéhyde, (55) l'anhydride maléique, (56) l'anhydride bromomaléique, (57) l'anhydride citraconique, (58) l'anhydride 2,3-diméthylmaléique, (59) l'anhydride dichloromaléique, (60) l'anhydride cis-aconitique, (61) l'anhydride itaconique, (62) l'anhydride méthylsuccinique, (63) l'anhydride acétylmercaptosuccinique, (64) l'anhydride 2,2-diméthylsuccinique, (65) l'anhydride phénylsuccinique, (66) l'anhydride 2-octèn-1-ylsuccinique, (67) l'anhydride 2-dodécèn-1-ylsuccinique, (68) l'anhydride 2-octadécèn-1-yl-succinique, (69) la 3-oxabicyclo[3.1.0]-hexane-2,4-dione, (70) l'anhydride diglycolique, (71) l'anhydride glutarique, (72) l'anhydride 3-méthylglutarique, (73) l'anhydride 2,2-diméthylglutarique, (74) l'anhydride 3,3-tétraméthylèneglutarique, (75) l'anhydride 1-cyclopentène-1,2-dicarboxylique, (76) l'anhydride 3,4,5,6-tétrahydrophtalique, (77) l'anhydride cis-1,2-cyclohexanedicarboxylique, (78) l'anhydride hexahydro-4-méthylphtalique, (79) l'anhydride méthyl-5-norbornène-2,3-dicarboxylique, (80) l'anhydride 2,3-pyridinecarboxylique, (81) l'anhydride 3,4-pyridinecarboxylique, (82) le furfurylmercaptan, (83) le thioacétate de S-furfuryle, (84) le sulfure de furfuryle, (85) le disulfure de furfuryle et de méthyle, (86) le disulfure de furfuryle, (87) le dimère de glycolaldéhyde, (88) la 6,7-dihydrocyclopenta1,3-dioxin-5(4H)-one, (89) la (2R,6R)-ter-butyl-6-méthyl-1,3-dioxan-4-one, (90) la 2,2-diméthyl-1,3-dioxane-4,6-dione, (91) la 3,6-diméthyl-1,4-dioxane-2,5-dione, (92) la 2,2,6-triméthyl-4H-1,3-dioxin-4-one, (93) la 2,2,5-triméthyl-1,3-dioxane-4,6-dione, (94) la 5-bromo-2,2,5-triméthyl-1,3-dioxane-4,6-dione, (95) le 1,3-dioxane-5,5-diméthanol, (96) le 1,3,5-trioxane, (97) la 1,6-dioxaspiro[4.4]nonane-2,7-dione, (98) la 1,4-dioxaspiro[4.5]décan-2-one, (99) le 1,7-dioxaspiro[5.5]undécane, (100) le 2,4,8,10-tétraoxaspiro[5.5]undécane, (101) le 3,9-divinyl-2,4,8-tétraoxaspiro[5.5]undécane, (102) le 2,2-pentaméthylène-1,3-dioxalane, (103) le 2-phényl-1,3-dioxalane, (104) le 1,4-cyclohexanedionemonoéthylèneacétal, (105) le 1,4-cyclohexanedionebis(éthylèneacétal), (106) le 1,4-cyclohexanedionemono-2,2-diméthyltriméthylèneacétal, (107) le pipéronal, (108) l'acétate de pipéronyle, (109) l'alcool pipéronylique, (110) le pipéronylnitrile, (111) la pipéronylamine, (112) le 6-nitropipéronal, (113) l'alcool 6-nitropipéronylique, (114) la 3',4'-(méthylènedioxy)acétophénone, (115) la 3,4-(méthylènedioxy)aniline, (116) le 2,3-(méthylènedioxy)benzaldéhyde, (117) le 3,4-(méthylènedioxy)phénylacétonitrile, (118) le 3,4-(méthylènedioxy)toluène et (119) des mélanges de ceux-ci ; ou dans lequel l'agent de transparence est un éther couronne ; ou dans lequel l'agent de transparence est choisi dans le groupe constitué par le 1,4,7,10-tétraoxacyclododécane (12-couronne-4), (2) le 2-(hydroxyéthyl)-12-couronne-4, (3) le 2-(aminoéthyl)-12-couronne-4, (4) le benzo-12-couronne-4, (5) le 1,4,7,10,13-pentaoxacyclododécane (15-couronne-5), (6) le 2-(hydroxyéthyl)-15-couronne-5, (7) le 2-(aminoéthyl)-15-couronne-5, (8) le benzo-15-couronne 5, (9) le 4'-aminobenzo-15-couronne-5, (10) le 4'-formylbenzo-15-couronne-5, (11) le 4'-nitrobenzo-15-couronne-5, (12) le pimélate de bis[(benzo-15-couronne-5)-15-ylméthyle], (13) le 1,4,7,10,13,16-hexaoxacyclooctadécane (18-couronne-6), (14) le 2-(aminoéthyl)-18-couronne-6, (15) le benzo-18-couronne-6, (16) le 4'-bromobenzo-18-couronne-6, (17) le dibenzo-18-couronne-6, (18) le di-tert-butyldibenzo-18-couronne-6, (19) le cis-dicyclohexane-18-couronne-6, (20) le dibenzo-24-couronne-8, (21) le dicyclohexano-24-couronne-8, (22) le dibenzo-30-couronne-10, et (23) des mélanges de ceux-ci ; ou dans lequel l'agent de transparence est un hydrocarbure cyclique ; ou dans lequel l'agent de transparence est choisi dans le groupe constitué par : (A) des matériaux répondant aux formules générales : dans lesquelles R₁, R₂, R₃, R₄, R₅, R₆, R₇, R₈, R₉, R₁₀, R₁₁, et R₁₂ sont choisis, chacun indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, R₁₀, R₁₁ et R₁₂ peuvent être liés ensemble pour former un cycle ; (B) des matériaux répondant à la formule générale : dans laquelle R₁, R₂, R₃, R₄, R₅ et R₆ sont choisis, chacun indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans laquelle deux ou plus de deux des symboles R₁, R₂, R₃, R₄, R₆ et R₆ peuvent être liés ensemble pour former un cycle ; (C) des matériaux répondant à la formule générale : dans lesquelles R₁, R₂, R₃, R₄, R₅, R₆, R₇, R₈, R₉, et R₁₀, sont choisis, chacun indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, et R₁₀ peuvent être liés ensemble pour former un cycle ; (D) des matériaux répondant aux formules générales : dans lesquelles R₁, R₂, R₃, R₄, R₅, R₆, R₇, R₈, R₉, R₁₀, R₁₁, et R₁₂, sont choisis, chacun indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, R₁₀, R₁₁,et R₁₂ peuvent être liés ensemble pour former un cycle ; (E) des matériaux répondant à la formule générale : dans laquelle R₁, R₂, R₃, R₄, R₅, R₆, R₇, R₈, R₉, R₁₀, sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans laquelle deux ou plus de deux des symboles R₁, R₂, R₃, R₄, R₅, R₆, R₇, R₈, R₉, et R₁₀, peuvent être liés ensemble pour former un cycle ; (F) des matériaux répondant aux formules générales : dans laquelle R₁, R₂, R₃, R₄, R₅, R₆, R₇, R₈, R₉ et R₁₀, sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, R₇, R₈, R₉, et R₁₀ peuvent être liés ensemble pour former un cycle ; (G) des matériaux répondant à la formule générale : dans laquelle la partie courbe de la structure représente une chaîne hydrocarbonée ou une chaîne hydrocarbonée substituée, dans laquelle deux ou plus de deux substituants peuvent être liés ensemble pour former un cycle ; et (H) des mélanges de ceux-ci ; ou dans lequel l'agent de transparence est choisi dans le groupe constitué par (1) le norbornane, (2) le 2-norbornanecarbonitrile, (3) le 2-norbornaneméthanol, (4) le 3-méthyl-2-norbornaneméthanol, (5) le camphène, (6) l'alcool fenchylique, (7) le thiocamphre, (8) le norbornène, (9) le 5-norbornène-2-carbonitrile, (10) le 5-norbornène-2-carboxaldéhyde, (11) le 5-norbornène-2-méthanol, (12) le 5-norbornène-2,2-diméthanol, (13) le 2-benzoyl-5-norbornène, (14) la 2-norbornanone, (15) la 3-chloro-2-norbornanone, (16) la fenchone, (17) le 3-(trifluoroacétyl)camphre, (18) le 3-heptafluorobutyrylcamphre, (19) le 3-bromocamphre, (20) le 9,10-dibromocamphre, (21) le 3,9,10-tribromocamphre, (22) le dicyclopentadiène, (23) le dimère de méthylcyclopentadiène, (24) le tricyclo[5.2.1]décane, (25) le 4,8-bis(hydroxyméthyl)tricyclo[5.2.1.0^{2,6}]décane, (26) le 8-cétotricyclo[5.2.1.0^{2,6}]décane, (27) la 3,4-diméthoxy-3-cyclobutène-1,2-dione, (28) la 3,4-diéthoxy-3-cyclobutène-1,2-dione, (29) la 3,4-diisopropoxy-3-cyclobutène-1,2-dione, (30) la 3,4-dibutoxy-3-cyclobutène-1,2-dione, (31) l'acide 3-méthyl-2-(nitrométhyl)-5-oxocyclopentaneacétique, (32) la 3-éthyl-2-hydroxy-2-cyclopentène-1-one, (33) le 4-méthoxy-2-oxo-3-cyclopentène-1-carboxylate de méthyle, (34) la 3,3a,6,6a-tétrahydro-2H-cyclopenta[b]furan-2-one, (35) la 3a,4,5,6a-hexahydro-5-hydroxy-4(hydroxyméthyl)-2H-cyclopenta[b]furan-2-one, (36) la 3-méthyl-1,2-cyclopentanedione, (37) le monohydrate de 4-hydroxy-5-méthyl-4-cyclopentène-1,3-dione, (38) la 2,4,4-triméthylcyclohexèn-1-one, (39) le 6-méthyl-2-oxo-3-cyclohexène-1-carboxylate d'éthyle, (40) le 4-hydroxy-6-méthyl-2-oxo-3-cyclohexène-1-carboxylate d'éthyle, (41) la 5-(1-acétoxy-1-méthyléthyl)-2-méthyl-2-cyclohéxène-1-one, (42) la thymoquinone, (43) la 2,6,6-triméthyl-2-cyclohexène-1,4-dione, (44) l'indane, (45) le 1-indanol, (46) le 2-indanol, (47) la 1-indanone, (48) la 2-indanone, (49) la 2-acétyl-1-tétralone, (50) la 4-méthyl-1-tétralone, (51) la 5,7-diméthyl-1-tétralone, (52) la 6,7-diméthoxy-1-tétralone, (53) la 1-méthyl-2-tétralone, (54) la 6,7-diméthoxy-2-tétralone, (55) la cyclohexanone, (56) la cycloheptanone, (57) la cyclooctanone, (58) la cyclononanone, (59) la cyclodécanone, (60) la cycloundécanone, (61) la cyclododécanone, (62) la cyclotridécanone, (63) la cyclopentadécanone, (64) la 2-acétylcyclohexanone, (65) la 2-allylcyclohexanone, (66) la 2-phénylcyclohexanone, (67) la cyclohexanedione, (68) la 2-acétyl-1,3-cyclohexanedione, (69) la 4,4-diméthyl-1,3-cyclohexanedione, (70) la 2-acétyl-1,3-cyclopentanedione, (71) la 3,3,5,5-tétraméthyl-1,2-cyclopentanedione, (72) la bicyclo[3.2.1]octan-2-one, (73) le 7-oxabicyclo[2.2.1]heptane-2,3-dicarboxylate d'endo-diméthyle, (74) le cinéole, (75) le bicyclo[2.2.2]oct-5-ène-2,3-diméthanol, (76) la tropone, (77) la tropolone, (78) l'oxyde de cyclooctène, (79) le 1,2,5,6-diépoxycyclooctane, (80) la 9-méthyl-Δ⁵⁽¹⁰⁾-octalin-1,6-dione, (81) la cis-bicyclo[3.3.0]octane-3,7-dione, (82)l'azulène, (83) la 1-benzosubérone, (84) le 1,5,9-cyclododécatriène, (85) l'époxyde de cyclododécane, (86) la 2,3-cyclododécénopyridine, (87) le 1,2,5,6,9,10-hexabromocyclododécane, (88) la 8-cyclohexadécène-1-one, (89) la bicyclo[10.3.0]pentadéc-12(1)-èn-13-one, (90) la 1,4,4a,8a-tétrahydro-endo-1,4-méthanonaphtalène-5,8-dione, et (91) des mélanges de ceux-ci ; ou dans lequel l'agent de transparence est une thiourée ; ou dans lequel l'agent de transparence est une sulfone ; ou dans lequel l'agent de transparence est un composé thiocyclique ; ou dans lequel l'agent de transparence est choisi dans le groupe constitué par des sulfites, des dérivés de sulfites, des sulfures, des dérivés de sulfures, des composés de soufre quaternaire, des dérivés de soufre quaternaire, et des mélanges de ceux-ci ; ou dans lequel l'agent de transparence est un composé thia-aza-cyclique ; ou dans lequel l'agent de transparence est choisi dans le groupe constitué par (1) la 1-allyl-2-thiourée, (2) la 1-méthallyl-3-méthyl-2-thiourée, (3) le 4-allyl-3-thiosemicarbazide, (4) la 1,3-diéthyl-2-thiourée, (5) la 1,3-dibutyl-2-thiourée, (6) la 1-benzyl-3-méthyl-2-thiourée, (7) la 1,1,3,3-tétraméthyl-2-thiourée, (8) le 2-imino-4-thiobiuret, (9) la 1-allyl-3-(2-hydroxyéthyl)-2-thiourée, (10) le bromhydrate de bromure de S-(2-aminoéthyl)isothiouronium, (11) le monohydrate de S,S-diphénylsulfillimine, (12) la méthylsulfone, (13) l'éthylsulfone, (14) la butylsulfone, (15) la butadiènesulfone, (16) la tétraméthylènesulfone, (17) la 1,4-butanesulfone, (18) le sulfate cyclique de 1,4-butanediol, (19) la benzylsulfone, (20) la phénylsulfone, (21) la phénylvinylsulfone, (22) la phénylstyrènesulfone, (23) la phényl-2-(triméthylsilyl)méthylsulfone, (24) la phényl-2-(triméthylsilyl)éthylsulfone, (25) la phényl-2-(triméthylsilyl)éthynylsulfone, (26) la 4-(fluorophényl)sulfone, (27) la 4-(fluorophényl)méthyl-sulfone, (28) la chlorométhylphénylsulfone, (29) la chlorométhyl-p-tolylsulfone, (30) la 2-chloroéthylphénylsulfone, (31) la méthylthiométhylphénylsulfone, (32) la méthylthiométhyl-p-tolylsulfone, (33) le 2-(phénylsulfonyl)tétrahydropyrane, (34) le 1-(phénylsulfonyl)indole, (35) le 1- (p-toluènesulfonyl)imidazole, (36) la 1-(p-tosyl)-3,4,4-triméthylimidazolidine, (37) la 4-(p-tosylsulfonyl)hexahydro-1,4-thiazépine, (38) le thionaphtène, (39) le 4-céto-4,5,6,7-tétrahydrothianaphtène, (40) le 2,2'-bithiophène, (41) le 2,2':5',2"-terthiophène, (42) la N-acétylhomocystéinethiolactone, (43) la tétrahydrothiopyran-4-one, (44) la thiochroman-4-one, (45) le thiochroman-4-ol, (46) l'acide thioctique, (47) le 1,3-dithiolane-2-carboxylate d'éthyle, (48) la 3H-1,2-benzodithiol-3-one, (49) le 1,3-dithiane, (50) le 2-phényl-1,3-dithiane, (51) le 1,3-dithiane-2-carboxylate d'éthyle, (52) la 5,6-dihydro-5-méthyl-4H-1,3,5-dithiazine, (53) le 1,4-dithiane, (54) le 2,5-dihydroxy-2,5-diméthyl-1,4-dithiane, (55) le 1,5-dithiacyclooactan-3-ol, (56) le 1,4-dithiaspiro-[45]-décan-8-ol, (57) le 1,3,5-trithiane, (58) le 1,4,7-trithiacyclononane, (59) le 1,4,7-trithiacyclodécane, (60) le 1,4,7,10-tétrathiacyclododécane, (61) le 3,6,9,14-tétrathiabicyclo[9.2.1]tétradéca-11,13-diène, (62) le 1,4,8,1-tétrathiacyclotétradécane, (63) le 1,5,9,13-tétrathiocyclohexadécane, (64) le 1,5,9,13-tétrathiacyclohexadécane-3,11-diol, (65) le 1,4,7,10,13-pentathiacyclopentadécane, (66) le 1,4,7,10,13,16-hexathiacyclooctadécane, (67) le 1,5,9,13,17,21-hexathiacyclotétracosane-3,11,19-triol, (68) le 1,4,7,10,13,16,19,22-octathiacyclotétracosane, (69) le 1,4,8,11,15,18,22,25-octathiacyclooctacosane, (70) le 1,4,7,10,13,16,19,22,25-nonathiacycloheptacosane, (71) le sulfite de diméthyle, (72) le sulfite de diéthyle, (73) le sulfite de sodium, (74) le disulfure d'allyle, (75) le disulfure d'aminophényle, (76) le disulfure de benzyle, (77) le sulfure de benzyle et de phényle, (78) le méthylsulfate de triméthylsulfonium, (79) l'iodure de (2-chloroéthyl)diméthylsulfonium, (80) le tétrafluoroborate de 3-(chloropropyl)diphénylsulfonium, (81) l'iodure de trimethylsulfonium, (82) l'iodure de triméthylsulfoxonium, (83) le chlorure de triméthyl- sulfoxonium, (84) le chlorure de triphénylméthane-sulfényle, (85) le bromure de diméthyl- (2-méthoxy-5-nitrobenzyl) sulfonium, (86) le perchlorate de thionine, (87) le p-xylylènebis(chlorure de tétrahydrothiophéneum), (88) le difluorotriméthylsilicate de tris(diméthylamino)sulfonium, (89) le trifluorométhylate de tris(diméthylamino)sulfonium, (90) le chlorure de (3-amino-3-carboxypropyl)diméthylsulfonium, et (91) des mélanges de ceux-ci ; ou dans lequel l'agent de transparence est un agent répondant à l'une des formules générales suivantes : dans lesquelles R₁, R₂, R₃, R₄, R₅, R₆ et R₇ sont choisis chacun, indépendamment des autres, dans le groupe constitué par des atomes d'hydrogène, des groupes alkyle, des groupes alkyle substitué, des groupes aryle, des groupes aryle substitué, des groupes arylalkyle, des groupes arylalkyle substitué, des groupes hydroxy, des groupes amine, des groupes imine, des groupes ammonium, des groupes pyridine, des groupes pyridinium, des groupes éther, des groupes aldéhyde, des groupes cétone, des groupes ester, des groupes amide, des groupes acide carboxylique, des groupes carbonyle, des groupes thiocarbonyle, des groupes sulfate, des groupes sulfonate, des groupes sulfure, des groupes sulfoxyde, des groupes phosphine, des groupes phosphonium, des groupes phosphate, des groupes cyano, des groupes nitrile, des groupes mercapto, des groupes nitroso, des atomes d'halogène, des groupes nitro, des groupes sulfone, des groupes acyle, des groupes anhydride d'acide et des groupes azide, dans lesquelles deux ou plus de deux des symboles R₁, R₂, R₃, R₄, R₅, R₆, et R₇, peuvent être liés ensemble pour former un cycle ; ou dans lequel l'agent de transparence est choisi dans le groupe constitué par (1) la 2-amino-2-thiazoline, (2) le 2-aminothiazole, (3) le 2-amino-4-méthylthiazole, (4) le 2-amino-4-méthylthiazole, (5) l'acide 2-amino-4-thiazolacétique, (6) le 2-acétamido-4-méthylthiazole, (7) le 2-acétylthiazole, (8) le 5-acétyl-2,4-diméthylthiazole, (9) le 4-méthyl-5-vinylthiazole, (10) le 2-amino-4-phényl-5-tétradécylthiazole, (11) la 2,4-thiazolidinedione, (12) la 3-aminorhodanine, (13) la 3-méthylrhodanine, (14) la 3-éthylrhodanine, (15) la 3-allylrhodanine, (16) la 3-hydroxy-4-méthyl-2(3H)-thiazoléthione, (17) le benzothiazole, (18) le 2-méthylbenzothiazole, (19) le 2-(méthylthio)benzothiazole, (20) le 2-amino-4-méthylbenzothiazole, (21) la 3-méthylbenzothiazole-2-thione, (22) le 2,1,3-benzothiadiazole, (23) le 4-amino-2,1,3-benzothiadiazole, (24) l'iodure de 3,4-diméthyl-5-(2-hydroxyéthyl)thiazolium , (25) le bromure de 3-éthyl-5-(2-hydroxyéthyl)4-méthylthiazolium, (26) le 2-amino-5-nitrothiazole, (27) l'acide 2-amino-α-(méthoxyimino)-4-thiazoleacétique, (28) le 2-amino-α-(hydroxyimino)-4-thiazoleacétate d'éthyle, (29) le 2-amino-α-(méthoxyimino)-4-thiazoleacétate d'éthyle, (30) le 2-amino-4-thiazoleacétate d'éthyle, (31) le 2-amino-4-thiazoleglyoxylate d'éthyle, (32) la 1-phényl-3-(2-thiazolyl)-2-thiourée, (33) le 2-amino-4-méthoxybenzothiazole, (34) le 2-amino-5,6-diméthylbenzothiazole, (35) le N'-(2-thiazolyl)sulfanilamide, le 6-éthoxy-2-benzothiazolesulfonamide, (37) le 2-(formylamino)-4-thiazoleacétate d'éthyle, (38) le 2-(formylamino)-4-thiazoleglyoxylate d'éthyle, (39) l'acide 2-(formylamino)-α-(méthoxyimino)-4-thiazoleacétique, (40) le chlorure de 2-acétamido-4-méthyl-5-thiazolesulfonyle, (41) l'acide 2-thioxo-4-thiazolidinecarboxylique, (42) l'acide thiazolidine-4-carboxylique, (43) la pseudothiohydantoïne, (44) le 2-amino-1,3,4-thiadiazole, (45) le 2-amino-5-trifluorométhyl-1,3,4-thiadiazole, (46) le 2-amino-5-méthyl-1,3,4-thiadiazole, (47) le 2-amino-5-éthyl-1,3,4-thiadiazole, (48), le 2-amino-5-(éthylthio)-1,3,4-thiadiazole, (49) le 5-amino-1,3,4-thiadiazole-2-thiol, (50) le 2-acétamido-5-benzylthio-1,3,4-thiadiazole, (51) le 5-acétamido-1,3,4-thiadiazole-2-sulfonamide, (52) le 5-anilino-1,2,3,4-thiatriazole, (53) le chlorhydrate de 2-amino-4,5-diméthylthiazole, (54) le chlorhydrate de 2-amino-4-imino-2-thiazoline, (55) le chlorhydrate de 2-amino-2-thiazoline, (56) le monohydrobromhydrate de 2-amino-5-bromothiazole, (57) le chlorhydrate de 5-amino-3-méthylisothiazole, (58) l'hydrate de chlorhydrate de 3-méthyl-2-benzothiazolinonehydrazone, (59) le dichlorhydrate de 5-amino-2-méthylbenzothiazole, (60) le monobromhydrate de 2,4-diamino-5-phénylthiazole, (61) le monohydrate de bromhydrate de 2-amino-4-phényl- thiazole, (62) le chlorhydrate de l'acide 2-(tritylamino)-α-(méthoxyimino)-4-thiazolacétique, (63) le chlorhydrate de 2,3,5,6-tétrahydro-6-phénylimidazo-[2,1-b]thiazole, (64) l'iodure de 3-éthyl-2-méthyl-2-thiazolium, (65) le chlorure de 3-benzyl-5-(2-hydroxyétyl)-4-méthylthiazolium, (66) le chlorhydrate de thiamine, (67) le bromure de 3-(carboxyméthyl)-benzothiazolium, (68) le tétrafluoroborate de 2-azido-3-éthylbenzothiazolium, (69) l'iodure de 3-éthyl-2-méthylbenzothiazolium, (70) l'iodure de 2-méthyl-3-propylbenzothiazolium, (71) le chlorure de 3-éthyl-2-(2-hydroxy-1-propényl)benzothiazolium, (72) le bromure de 3,6-diméthyl-2- (4-diméthylaminophényl)benzothiazolium, (73) le dichlorhydrate de trifluoropérazine, (74) le chlorhydrate de thioridazine, (75) le chlorhydrate de prométhazine, (76) le chlorhydrate d'éthopropazine, (77) le chlorhydrate de chlorpromazine, et (78) des mélanges de ceux-ci ; ou dans lequel l'agent de transparence est choisi dans le groupe constitué par des phospines, des phosphites, des composés de phosphore cycliques, des oxydes de phosphine, des sels de phosphonium quaternaire, et des mélanges de ceux-ci ; ou dans lequel l'agent de transparence est choisi dans le groupe constitué par (1) la triphénylphosphine, (2) la tri-m-tolylphosphine, (3) la tris(3-méthoxyphényl)phosphine, (4) la tris(4-chlorophényl)phosphine, (5) la tris(pentafluorophényl)phosphine, (6) la tricyclohexylphosphine, (7) la tribenzylphosphine, (8) la tri-2-furylphosphine, (9) la bis(pyrrolidino)méthoxyphosphine, (10) la tétraphénylbiphosphine, (11) le 1,3-bis(diphénylphosphino)propane, (12) le 1,5-bis(diphénylphosphino)pentane, (13) le 1,6-bis(diphénylphosphino)hexane, (14) l'isopropyldiphénylphosphine, (15) la diphényl(p-tolyl)-phosphine, (16) la (4-bromophényl)diphénylphosphine, (17) la diphényl-2-pyridylphosphine, (18) la dicyclohexylphénylphosphine, (19) le phosphite de triméthyle, (20) le phosphite de triéthyle, (21) le phosphite de tris(2-chloroéthyle), (22) le phosphite de tributyle, (23) le phosphite de triphényle, (24) le phosphite de triméthyle-iodure de cuivre, (25) le phosphite de triéthyle-iodure de cuivre, (26) le phosphite de dipropyle, (27) le phosphite de bis(2-éthylhexyle), (28) le phosphite de bis(4-nitrobenzyle), (29) le fluorophosphite de 2,2'-éthylidènebis(4,6-di-tert-butylphényle), (30) le diphosphite de pentaérythrol et de diphényle, (31) le phosphorodiamidate de 2-furyle et de tétraméthyle, (32) le (pyrrolidinométhyle)phosphonate de diéthyle, (33) le monohydrate de cyclophosphamide, (34) le 2-oxyde de 2-chloro-1,3,2-dioxaphospholane, (35) la N,N-diéthyl-1,5-dihydro-2,4,3-benzodioxaphosphépin-3-amine, (36) le 1,2-phénylènephosphochloridite, (37) le phosphochloridate de 1,2-phénylène, (38) la 2-chloro-4H-1,3,2-benzodioxaphosphorin-4-one, (39) le 2,4-disulfure de 2,4-bis(méthylthio)-1,3-dithia-2,4-diphosphétane, (40) l'oxyde de triphénylphosphine, (41) l'oxyde de tris(hydroxyméthyl)phosphine, (42) l'oxyde de triméthoxyphosphine, (43) l'oxyde de triéthoxyphosphine, (44) l'oxyde de triphénoxyphosphine, (45) l'oxyde de tris (2-butoxyéthoxy)phosphine, (46) l'oxyde de diphénylphosphine, (47) l'oxyde de diphényl(2,4,6-triméthylbenzoyl)phosphine, (48) l'acide phénylphosphinique, (49) le phosphate de diphényle, (50) l'acide vinylphosphonique, (51) l'acide propylphosphonique, (52) l'acide pyrophosphorique, (53) le phosphate de triphényle, (54) le chlorure de tétrabutylphosphonium, (55) le bromure de tétrabutylphosphonium, (56) le bromure d'hexadécyltributylphosphonium, (57) le bromure de stéaryltributylphosphonium, (58) le bromure d'azidotris(diéthylamino)phosphonium, (59) le trimère de chlorure phosphonitrilique, (60) le bromure de tétraméthylphosphonium, (61) le chlorure de tétraméthylphosphonium, (62), le bromure de tétraéthylphosphonium, (63) le chlorure de tétraéthylphosphonium, (64) l'iodure de tétraéthylphosphonium, (65) le bromure de tétraphénylphosphonium, (66) le chlorure de tétraphénylphosphonium (67) l'iodure de tétraphénylphosphonium, (68) le bromure de méthyltriphénylphosphonium, (69) l'iodure de méthyltriphénylphosphonium, (70) le bromure d'éthyltriphénylphosphonium, (71) le bromure de n-propyltriphénylphosphonium, (72) l'iodure d'isopropyltriphénylphosphonium, (73) le bromure de cyclopropyltriphénylphosphonium, (74) le bromure de n-butyltriphénylphosphonium, (75) le bromure d'isobutyltriphénylphosphonium, (76) le bromure d'hexyltriphénylphosphonium, (77) le chlorure de benzyltriphénylphosphonium, (78) le bromure de bromométhyltriphénylphosphonium, (79) le chlorure de chlorométhyltriphénylephosphonium, (80) le bromure de 3-bromopropyltriphénylphosphonium, (81) le bromure de 3-bromobutyltriphénylphosphonium, (82) le bromure de 4-bromobutyltriphénylphosphonium, (83) le bromure de 2-diméthylaminoéthyltriphénylphosphonium, (84) le bromure de [(3-diméthylamino)propyl]triphénylphosphonium, (85) le bromure de 2-hydroxyéthyltriphénylphosphonium, (86) le chlorure de (2-hydroxyéthyl)triphénylphosphonium, (87) le bromure de [3-hydroxy-2-méthylpropyl]-triphénylphosphonium, (88) le bromure de [3-hydroxy-2-méthylpropyl]triphénylphosphonium, (89) le bromure de (2-hydroxybenzyltriphénylphosphonium, (90) le chlorure de (formylméthyl)triphénylphosphonium, (91) le chlorure de (méthoxyméthyl)triphénylphosphonium, (92) le chlorure d'acétonyltriphénylphosphonium, (93) le bromure de carbométhoxyméthyltriphénylphosphonium, (94) le chlorure d' (éthoxycarbonylméthyl)triphénylphosphonium, (95) le bromure de carbéthoxyméthyltriphénylphosphonium, (96) le bromure de (tert-butoxycarbonylméthyl)triphénylphosphonium, (97) le bromure de phénacyltriphénylphosphonium, (98) le bromure de 4-éthoxybenzyl)triphénylphosphonium, (99) le bromure de 4-butoxybenzyltriphénylphosphonium, (100) le bromure de 2-(1,3-dioxan-2-yl)éthyl]triphénylphosphonium, (101) le bromure de (1,3-dioxolan-2-ylméthyl)triphénylphosphonium, (102) le bromure de vinyltriphénylphosphonium, (103) le bromure d'allyltriphénylphosphonium, (104) le chlorure d'allyltriphénylphosphonium, (105) le bromure de propargyltriphénylphosphonium, (106) le bromure de (3-triméthylsilyl-2-propynyl)triphénylphosphonium, (107) le p-xylylènebis(bromure de triphénylphosphonium), et (108) des mélanges de ceux-ci ; ou dans lequel l'agent de transparence est un nitrile ; ou dans lequel l'agent de transparence est choisi dans le groupe constitué par le cyanoacétohydrazide, (2) le 4,4-diméthyl-3-oxopentanenitrile, (3) le 1-cyano-N-méthylthioformamide, (4) le N,N-diméthyldithiocarbamate de cyanométhyle, (5) le 4-hydroxy-3-méthoxyphénylacétonitrile, (6) le cyanure de tosyle, (7) l'isocyanure de tosylméthyle, (8) le 5-fluoro-2-méthylbenzonitrile, (9) le 2-fluoro-5-méthylbenzonitrile, (10) le 4-(méthylthio)benzonitrile, (11) le 4-(diméthylamino)benzonitrile, (12) le 3,4-diméthoxybenzonitrile, (13) le 4-hydroxy-3-méthoxybenzonitrile, (14) le 4-(trans-4-pentyl-cyclohexyl)benzonitrile, (15) le 4'-pentyl-4'-biphénylcarbonitrile, (16) le 4'-(pentyloxy)-4-biphénylcarbonitrile, (17) le 4'-hexyl-4-biphénylcarbonitrile, (18) le 4'-(hexyloxy)-4-biphényl-carbonitrile, (19) le 4'-heptyl-4-biphénylcarbonitrile, (20) le 4'-heptyloxy-4-biphénylcarbonitrile, (21) le 4'-octyl-4-biphénylcarbonitrile, (22) le 4'-(octyloxy)-4-biphénylcarbonitrile, (23) le succinonitrile, (24) le fumaronitrile, (25) le 1,4-dicyano-2-butène, (26) le (diméthylaminométhylène)malononitrile, (27) le (1-éthoxyéthylidène)malononitrile, (28) l'α-chlorobenzylidènemalononitrile, (29) le benzylidènemalononitrile, (30) le 2-benzoyloxy-2-phényl-malononitrile, (31) l'O-(p-tosyl)isonitrosomalononitrile, (32) le tétrafluorophtalonitrile, (33) l'iminodiacétonitrile, (34) le phénylènediacétonitrile, (35) le 3,3' - (4-formylphénylimino)dipropionitrile, (36) le tris(2-cyanoéthyl)nitrométhane, (37) le 1,1,3,3-propanetétracarbonitrile, (38) l'oxyde de tétracyanoéthylène, et (39) des mélanges de ceux-ci, ou dans lequel l'agent de transparence est choisi dans le groupe constitué par des isothiocyanates, des isocyanates, et des mélanges de ceux-ci ; ou dans lequel l'agent de transparence est choisi dans le groupe constitué par (1) l'isothiocyanate de 4-azidophényle, (2) l'isothiocyanate de 1-naphtyle, (3) l'isothiocyanate de 4-diméthylamino-1-naphtyle, (4) le 1-isothiocyanato-4-(trans-4-propylcyclohexyl)benzène, (5) le 1-(trans-4-hexyl-cyclohexyl)-4-isothiocyanatobenzène, (6) le 1-(4-trans-hexylcyclohexyl) -4-[2- (4-isothiocyanatophényl)]benzène, (7) le 1-isothiocyanato-4(trans-4-octylcyclohexyl)benzène, (8) le 4-pentabicyclo[2.2.2]octane-1-carboxylate de 4-isothiocyanatophényle, (9) le thiocyanate de benzyle, (10) le thiocyanate de guanidine, (11) le dithiocyanate de méthylène, (12) le 4,4'-méthylènebis(isocyanate de phényle), (13) le 4,4'-méthylènebis (isocyanate de 2,6-diéthyle), et (14) des mélanges de ceux-ci ; ou dans lequel l'agent de transparence est choisi dans le groupe constitué par des composés d'oxime, des composés d'acide hydroxamique, et des mélanges de ceux-ci ; ou dans lequel l'agent de transparence est choisi dans le groupe constitué par (1) le formamidoxime, (2) l'acétaldoxime, (3) le pyruvaldéhyde-1-oxime, (4) l'acétoneoxime, (5) le chlorooximidoacétate d'éthyle, (6) le 2,3-butanedionemonooxime, (7) le 5-hydroxypenténaloxime, (8) le cyclopentanoneoxime, (9) le cyclohexanoneoxime, (10) le cyclooctanoneoxime, (11) le benzaldéhydeoxime, (12) le 2-nitrobenzaldéhydeoxime, (13) le salicylaldoxime, (14) la 2-isonitrosoacétophénone, (15) le 1-phényl-1,2-propanedione-2-oxime, (16) le 2-pyridinealdoxime, (17) le nifuroxime, et (18) des mélanges de ceux-ci ; ou dans lequel l'agent de transparence est un dérivé d'acide hydroxamique ; ou dans lequel l'agent de transparence est choisi dans le groupe constitué par (1) l'acide acétohydroxamique, (2) l'acide subérohydroxamique, (3) l'acide mandélohydroxamique, (4) l'acide benzohydroxamique, (5) l'acide N-phénylbenzohydroxamique, et (6) des mélanges de ceux-ci ; ou dans lequel l'agent de transparence est choisi dans le groupe constitué par des sels d'alkylammonium, des sels d'arylammonium, des sels d'arylalkylammonium, et des mélanges de ceux-ci ; ou dans lequel l'agent de transparence est choisi dans le groupe constitué par (1) le tétrahydrate de fluorure de tétraméthylammonium, (2) le tétrahydrate d'acétate de tétraéthylammonium, (3) le chlorure de tétrabutylammonium, (4) l'hydrate de chlorure de tétrabutylammonium, (5) le bromure de tétrabutylammonium, (6) le tribromure de tétrabutylammonium, (7) l'acétate de tétrabutylammonium, (8) le thiocyanate de tétrabutylammonium, (9) le bromure de tétrapentylammonium, (10) le bromure de tétrahexylammonium, (11) le chlorure de tétrahexylammonium, (12) le sulfate acide de tétrahexylammonium, (13) le chlorure de tétraheptylammonium, (14) le bromure de tétraheptylammonium, (15) le bromure de tétraoctylammonium, (16) le bromure de tétrakisdécylammonium, (17) le bromure de tétrahexadécylammonium, (18) le bromure de tétraméthylammonium, (19) le chlorure de tétraméthylammonium, (20) l'iodure de tétraméthylammonium, (21) le bromure de tétraéthylammonium, (22) le chlorure de tétraéthylammonium, (23) l'iodure de tétraéthylammonium, (24) le bromure de tétrapropylammonium, (25) l'iodure de tétrapropylammonium, (26) l'iodure de tétrabutylammonium, (27) le chlorure de tétrapentylammonium, (28) le bromure de tétrahexylammonium, (29) l'iodure de tétrahexylammonium, (30) le bromure de tétradécylammonium, (31) le bromure de tétradodécylammonium, (32) le bromure de tétraoctadécylammonium, (33) le bromure de méthyltrioctylammonium, (34) le chlorure de' tridodécylméthylammonium, (35) l'iodure de tridodécylméthylammonium, (36) le bromure de N-dodécyl-N-méthyléphédrinium, (37) le tribromure de phényltriméthylammonium, (38) le chlorure de tricaprylméthylammonium, (39) le chlorure de tridodécylméthylammonium, (40) le chlorure de tridécyloxypropyldihydroxyéthylméthylammonium, (41) le chlorure de N-tétradécyldiméthylnaphtylméthylammonium, (42) le chlorure de d'octadécyldiéthanolméthylammonium, (43) le chlorure d'octadécyldihydroxyéthylméthylammonium, (44) le chlorure de suif dihydrogéné-benzylméthylammonium, (45) le chlorhydrate de chlorure de 2-aminoéthyltriméthylammonium, (46) le bromure de 2-bromoéthyltriméthylammonium, (47) le chlorure de 2-chloroéthyltriméthylammonium, (48) le chlorure de 3-carboxypropyltriméthylammonium, (49) le chlorure de [3-(méthacryloylamino)propyl]triméthylammonium, (50) le bromure de phényltriméthylammonium, (51) le chlorure de phényltriméthylammonium, (52) l'iodure de phényltriméthylammonium, (53) le chlorure de benzyltriméthylammonium, (54) le bromure de benzyltriméthylammonium, (55) le chlorure de 4-nitrobenzyltriméthylammonium, (56) l'iodure de [2-(4-nitrophényl)allyl]triméthylammonium, (57) le chlorure de coco-triméthylammonium, (58) le chlorure de palmityltriméthylammonium, (59) le bromure de myristyltriméthylammonium, (60) le chlorure d'oléyltriméthylammonium, (61) le chlorure de soya-triméthylammonium, (62) le chlorure de suif-triméthylammonium, (63) le chlorure de suif hydrogéné-triméthylammonium, (64) le chlorure de stéaryltriméthylammonium, (65) le chlorure de béhényltriméthylammonium, (66) le chlorure de guar-hydroxypropyltriméthylammonium, (67) le bromure de benzyltriéthylammonium, (68) le bromure de butyltripropylammonium, (69) le chlorure de méthyltributylammonium, (70) le bromure de méthyltributylammonium, (71) l'iodure de méthyltributylammonium, (72) le chlorure de benzyltributylammonium, (73) le bromure de benzyltributylammonium, (74) l'iodure de benzyltributylammonium, (75) le bromure d'heptyltributylammonium, (76) le bromure de benzyldodécyldiméthylammonium, (77) le dihydrate de chlorure de benzyltétradécylediméthylammonium, (78) le monohydrate de chlorure de benzylcétyldiméthylammonium, (79) le monohydrate de chlorure de benzylstéaryldiméthylammonium, (80) le chlorure de N,N-diméthylméthylèneammonium, (81) l'iodure de N,N-diméthylméthylèneammonium, (82) le chlorure de chlorométhylènediméthylammonium, (83) le chlorure de dichlorométhylènediméthylammonium, (84) le chlorure de diméthylaminométhylèneaminométhylènediméthylammonium, (85) le chlorure de benzéthonium, (86) le chlorure de méthylbenzéthonium, (87) le chlorure de 1-propanaminium-2,3-dihydroxy-N-diméthyl-N-[3 (oxococoyl) aminopropyle], (88) le bromure de cétyldiméthyléthylammonium, (89) le chlorure d'octyldodécyldiméthylammonium, (90) le bromure de dodécyl-(2-hydroxy-1-méthyl-2-phényléthyl)diméthylammonium, (91) le bromure de dodécyldiméthyl-2-phénoxyéthylammonium, (92) le chlorure de dodécanoyl-N-méthylaminoéthyl(phénylcarbamylméthyl)diméthylammonium, (93) le chlorure de 3-chloro-2-hydroxypropyl-N,N,N-diméthyldodécylammonium, (94) le chlorure de 3-chloro-2-hydroxypropyl-N,N,N-diméthyloctadécylammonnium, (95) le bromure de dodécylbenzyldiméthylammonium, (96) le chlorure de dodécylbenzyldiméthylammonium, (97) le chlorure de coco-benzyldiméthylammonium, (98) le chlorure de benzyltétradécyldiméthylammonium, (99) le chlorure de benzylcétyldiméthylammonium, (100) le chlorure de benzyloctadécyldiméthylammonium, (101) le chlorure de benzyl-suif-diméthylammonium, (102) le chlorure de benzyl-suif hydrogéné-diméthylammonium, (103) le chlorure de benzyl-béhényldiméthylammonium, (104) le chlorure de dioctyldiméthylammonium, (105) le chlorure de didécyldiméthylammonium, (106) le bromure de didécyldiméthylammonium, (107) le chlorure de dicoco-diméthylammonium, (108) le chlorure de dicétyldiméthylammonium, '(109) le chlorure de disoya-diméthylammonium, (110) le chlorure de disuif-diméthylammonium, (111) le chlorure de suif dihydrogénédiméthylammonium, (112) le chlorure de dibéhényl/diarachidyldiméthylammonium, (113) le chlorure de soya-amidopropylbenzyldiméthylammonium, (114) le chlorure de soja-di-coco-ammonium quaternaire, (115) le chlorure de gluco-namidopropyldiméthyl-2-hydroxyéthylammonium, (116) un chlorure de N-alkyl-N-N-diméthyl-N-(acétate de dodécylammonium), dans lequel le groupe alkyle comporte de 14 à 20 atomes de carbone, (117) le chlorure de visonamidopropyldiméthyl-2-hydroxyéthylammonium, (118) le chlorure de N-colza-(3-amidopropyl)-N-N-diméthyl-N-(2,3-époxypropyl)ammonium, (119) le chlorure de N-stéaryl-(3-amidopropyl)-N-benzyldiméthylammonium, (120) le chlorure de colza-amidopropylbenzyldiméthylammonium, (121) le chlorure de colza-amidopropyléthyldiméthylammonium, (122) le phosphate de chlorure de coco-amidopropylpolyéthylèneglycoldiméthylammonium, (123) le chlorure de butyrylcholine, et (124) des mélanges de ceux-ci ; ou dans lequel l'agent de transparence est choisi dans le groupe constitué par le thiocyanate de pipéridine, le 2-pipéridineméthanol, la bis(pentaméthylène)urée, le 4,4'-triméthylènebis(1-pipéridinepropionitrile), l'oxyde de tripipéridinophosphine, l'homopipérazine, la 1-pipéronylpipérazine, le trisulfate d'hexacylène, la 5,10,15,20-tétraphényl-21H,23H-porphine, la 5,10,15,20-tétrakis(4-méthoxyphényl)-2H,23H-porphine, le pyrrole-2-carboxaldéhyde, le 3-pyrrolidino-1,2-propanediol, le pyrazole, le 3-aminopyrazole, l'imidazole, le 2-éthylimidazole, la 2-(2-pipéridinoéthyl)pyridine, le chlorure de 1-dodécylpyridinium, le perbromure de bromure de pyridinium, la 3-aminoquinoléine, la 8-hydroxyquinoléine, la 7,8-benzoquinoléine, la 8-hydroxyquinaldine, la quinoxaline, le monohydrate de 4,5-dihydro-6-méthyl-3(2H)-pyridazinone, la phtalazine, la 1,10-phénanthroline, la 1,3,5-triazine, la trichloromélamine, l'acide trichloroisocyanurique, le norbornane, le tricyclo-[5.2.1.0]décape, le norcamphre, la tropolone, le 1-indanol, le trans,trans,cis-1,5,9-cyclododécatriène, l'époxyde de cyclodécane, la 2,3-cyclododécanepyridine, le 1,2,5,6,9,10-hexabromocyclododécane, la 1,4,4a,8a-tétrahydro-endo-1,4-méthanonaphtalène-5,8-dione, la γ-butyrolactone, la β,β-diméthyl-γ-(hydroxyméthyl)-γ-buty-rolactone, la 2,5-diméthyl-4-hydroxy-3(2H)-furanone, le dihydrate d'hydrindantine, le 2,4,8,10-tétraoxaspiro-[5.5]undécane, le 1,3,5-trioxane, la cyclooctanone, le pipéronal, l'alcool pipéronylique, le pipéronylnitrile, le 3,4(méthylènedioxy)phénylacétonitrile, l'anhydride maléique, l'anhydride s-acétylmercaptosuccinique, l'anhydride 2-octadécèn-1-ylsuccinique, le 18-couronne-6, le benzo-18-couronne-6, le dibenzo-18-couronne-6, le dibenzo-24-couronne-8, le 5-amino-3-méthylisooxazole, la 2-oxazolidone, la 5,5-diméthyloxazolidine-2,4-dione, la 3-éthyl-2-thioxo-4-oxazolidinone, le 3-morpholino-1,2-propanediol, la 4-phénylmorpholine, le N,N'-dibenzyl-1,4,10,13-tétraoxa-7,16-diazacyclooctadécane, le 4,7,13,16,21,24-hexaoxa-1,10-diazabicyclo[8.8.8]hexacosane, le γ-valérolactame, l'ε-caprolactame, la 2-azacyclooctanone, la 2-azacyclononanone, le maléimide, le n-méthylsuccinimide, un sel de DBU-phtalimide, la 1-allyl-2-thiourée, le 1,3-dithiane, la 1-benzyl-3-méthyl-2thiourée, le 2-imino-4-thiobiuret, la butylsulfone, le 2,2'-bithiophène, le 2-phényl-1,3-dithiane, le 3,6,9,14-tétrathiabicyclo[9.2.1]tétradéca-11,13-diène, le 1,5,9,13-tétrathiacyclohexadécane-3,11-diol, le 1,4,7,10,13-pentathiacyclopentadécane, le 2-aminothiazole, la 2-amino-2-thiazoline, la 3-méthylrhodanine, le bromure de 3-éthyl-5-(2-hydroxyéthyl)-4-méthylthiazolium, la triphénylphosphine, la tricyclohexylphosphine, le 1,3-bis(diphénylphosphino)propane, le 1,5-bis(diphénylphosphino)pentane, l'isopropyldiphénylphosphine, le phosphite de triéthyle, le phosphite de triphényle, le phosphite de triéthyle-iodure de cuivre, le phosphite de dipropyle, le phosphite de bis(2-éthylhexyle), le phosphite de bis(4-nitrobenzyle), l'oxyde de diphénylphosphine, l'oxyde de diphényl-(2,4,6-triméthylbenzoyl)phosphine, l'acide vinylphosphonique, le cyanoacétohydrazide, le N,N-diméthyldithiocarbamate de cyanométhyle, le 4'-pentyl-4'-biphénylcarbonitrile, le 4'-(octyloxy)-4-biphénylcarbonitrile, le 1,4-dicyano-2-butène, le benzylidènemalononitrile, le 1-isothiocyanato-4-(trans-4-propylcyclohexyl)benzène, le formamidoxime, le chlorooximidoacétate d'éthyle, l'acide acétohydroxamique, le chlorure de tétrahexylammonium, le chlorure de tétraheptylammonium, le bromure de tétraheptylammonium et des mélanges de ceux-ci.

9. Procédé qui comprend les étapes consistant à (1) fournir l'élément de formation d'images par migration selon la revendication 1, comprenant (a) un substrat, (b) une couche ramollissable comprenant un matériau ramollisable et un matériau de marquage par migration photosensible, et (c) un agent de transparence qui rend transparent le matériau de marquage par migration en contact avec lui, contenu dans au moins une couche de l'élément de formation d'images par migration ; (2) charger uniformément l'élément de formation d'images ; (3) à la suite de l'étape (2), exposer l'élément de formation d'images chargé à un rayonnement activant à une longueur d'onde à laquelle le matériau de marquage par migration est sensible ; (4) à la suite de l'étape (3), provoquer le ramollissement du matériau ramollissable et permettre à une première partie du matériau de marquage par migration de migrer à travers le matériau ramollissable vers le substrat selon un motif formant une image tandis qu'une seconde partie du matériau de marquage par migration reste essentiellement sans avoir migré à l'intérieur de la couche ramollissable, dans lequel à la suite de la migration de la première partie du matériau de marquage par migration, (a) la première partie du matériau de marquage par migration entre en contact avec l'agent de transparence et la seconde partie du matériau de marquage par migration n'entre pas en contact avec l'agent de transparence ; ou (b) la seconde partie du matériau de marquage par migration entre en contact avec l'agent de transparence et la première partie du matériau de marquage par migration n'entre pas en contact avec l'agent de transparence

10. Procédé selon la revendication 9, dans lequel la première partie du matériau de marquage par migration entre en contact avec l'agent de transparence et la seconde partie du matériau de marquage par migration n'entre pas en contact avec l'agent de transparence ; ou dans lequel la seconde partie du matériau de marquage par migration entre en contact avec l'agent de transparence et la première partie du matériau de marquage par migration n'entre pas en contact avec l'agent de transparence.
